

# United States Patent [19]

Aoike et al.

[11] Patent Number: 4,882,251

[45] Date of Patent: Nov. 21, 1989

[54] LIGHT RECEIVING MEMBER HAVING A MULTILAYERED LIGHT RECEIVING LAYER COMPOSED OF A LOWER LAYER MADE OF ALUMINUM-CONTAINING INORGANIC MATERIAL AND AN UPPER LAYER MADE OF NON-SINGLE-CRYSTAL SILICON MATERIAL

[75] Inventors: Tatsuyuki Aoike; Masafumi Sano; Takehito Yoshino; Toshimitsu Kariya; Hiroaki Niino, all of Nagahama, Japan

[73] Assignee: Canon Kabushiki Kaisha, Tokyo, Japan

[21] Appl. No.: 183,701

[22] Filed: Apr. 19, 1988

[30] Foreign Application Priority Data

Apr. 22, 1987 [JP] Japan ..... 62-99547  
Apr. 27, 1987 [JP] Japan ..... 62-104915  
May 6, 1987 [JP] Japan ..... 62-111622  
May 7, 1987 [JP] Japan ..... 62-112159  
Jun. 29, 1987 [JP] Japan ..... 62-161538  
Aug. 5, 1987 [JP] Japan ..... 62-196566  
Aug. 6, 1987 [JP] Japan ..... 62-197829  
Dec. 16, 1987 [JP] Japan ..... 62-316312

[51] Int. Cl.<sup>4</sup> ..... G03G 5/082; G03G 5/14

[52] U.S. Cl. ..... 430/57; 430/60;  
430/65

[58] Field of Search ..... 430/57, 60, 65

[56]

## References Cited

### U.S. PATENT DOCUMENTS

4,460,669 7/1984 Ogawa et al. ..... 430/57

### FOREIGN PATENT DOCUMENTS

59-28162 2/1984 Japan ..... 430/60

Primary Examiner—Roland E. Martin

Attorney, Agent, or Firm—Fitzpatrick, Cella, Harper & Scinto

[57]

## ABSTRACT

A light receiving member for electrophotography made up of an aluminum support and a multilayered light receiving layer exhibiting photoconductivity formed on the aluminum support, wherein the multilayered light receiving layer consists of a lower layer in contact with the support and an upper layer, the lower layer being made of an inorganic material containing at least aluminum atom (Al), silicon atoms (Si) and hydrogen atoms (H), and having portion in which the aluminum atoms (Al), silicon atoms (Si), and hydrogen atoms (H) are unevenly distributed across the layer thickness, the upper layer being made of a non-single-crystal material composed of silicon atoms (Si) as the matrix and at least either of hydrogen atoms (H) or halogen atoms (X) and containing atoms to control conductivity in the layer region in adjacent with the lower layer. The light receiving member for electrophotography can overcome all of the foregoing problems and exhibits extremely excellent electrical property, optical property, photoconductivity, durability, image property and circumstantial property of use.

30 Claims, 17 Drawing Sheets



FIG. 1



FIG. 2



FIG. 3



FIG. 4



FIG. 5



FIG. 6



FIG. 7



FIG. 8



FIG. 9



FIG. 10



FIG. 11



FIG. 12



FIG. 13



FIG. 14



FIG. 15



FIG. 16



FIG. 17



FIG. 18



FIG. 19



FIG. 20



FIG. 21



FIG. 22



FIG. 23



FIG. 24



FIG. 25



FIG. 26



FIG. 27



FIG. 28



FIG. 29



FIG. 30



FIG. 31



FIG. 32



FIG. 33



FIG. 34



FIG. 35



FIG. 36



FIG. 37



FIG. 38



FIG. 39



FIG. 40





FIG. 42



FIG. 43 (c)



FIG. 43 (d)



**LIGHT RECEIVING MEMBER HAVING A  
MULTILAYERED LIGHT RECEIVING LAYER  
COMPOSED OF A LOWER LAYER MADE OF  
ALUMINUM-CONTAINING INORGANIC  
MATERIAL AND AN UPPER LAYER MADE OF  
NON-SINGLE-CRYSTAL SILICON MATERIAL**

**FIELD OF THE INVENTION**

This invention concerns a light receiving member sensitive to electromagnetic waves such as light (which herein means in a broader sense those lights such as ultraviolet rays, visible rays, infrared rays, X-rays, and  $\gamma$ -rays).

More particularly, it relates to an improved light receiving member having a multilayered light receiving layer composed of a lower layer made of an inorganic material containing at least aluminum atoms, silicon atoms, and hydrogen atoms, and an upper layer made of non-single-crystal silicon material, which is suitable particularly for use in the case where coherent lights such as laser beams are applied.

**BACKGROUND OF THE INVENTION**

The light receiving member used for image formation has a light receiving layer made of a photoconductive material. This material is required to have characteristic properties such as high sensitivity, high S/N ratio (ratio of light current ( $I_p$ ) to dark current ( $I_d$ )), absorption spectral characteristic matching the spectral characteristic of electromagnetic wave for irradiation, rapid optical response, appropriate dark resistance, and non-toxicity to the human body at the time of use. The non-toxicity at the time of use is an important requirement in the case of a light receiving member for electronic photography which is built into an electronic photographic apparatus used as an office machine.

A photoconductive material attracting attention at present from the standpoint mentioned above is amorphous silicon (A-Si for short hereinafter). The application of A-Si to the light receiving member for electrophotography is disclosed in, for example, German Patent Laid-open Nos. 2746967 and 2855718.

FIG. 2 is a schematic sectional view showing the layer structure of the conventional light receiving member for electrophotography. There are shown an aluminum support 201 and a photosensitive layer of A-Si 202. This type of light receiving member for electrophotography is usually produced by forming the photosensitive layer 202 of A-Si on the aluminum support 201 heated to 50°-350° C., by deposition, hot CVD process, plasma CVD process, plasma CVD process or sputtering.

Unfortunately, this light receiving member for electrophotography has a disadvantage that the sensitive layer 202 of A-Si is liable to crack or peel off during cooling subsequent to the film forming step, because the coefficient of thermal expansion of aluminum is nearly ten times as high as that of A-Si. To solve this problem, there was proposed a photosensitive body for electrophotography which is composed of an aluminum support, an intermediate layer containing at least aluminum and a sensitive layer of A-Si (Japanese Patent Laid-open No. 28162/1984). The intermediate layer containing at least aluminum relieves the stress arising from the difference in the coefficient of thermal expansion between the aluminum support and the A-Si sensitive

layer, thereby reducing the cracking and peeling of the A-Si sensitive layer.

The conventional light receiving member for electrophotography which has the light receiving layer made of A-Si has been improved in electrical, optical, and photoconductive characteristics (such as dark resistance, photosensitivity, and light responsivity), adaptability of use environment, stability with time, and durability. Nevertheless, it still has room for further improvement in its overall performance.

For the improvement of image characteristics, several improvements have recently been made on the optical exposure unit, development unit, and transfer unit in the electrophotographic apparatus. This, in turn, has required the light receiving member for electrophotography to be improved further in image characteristics. With the improvement of images in resolving power, the users have begun to require further improvements such as the reduction of unevenness (so-called "coarse image") in the region where the image density delicately changes, and the reduction of image defects (so-called "dots") which appear in black or white spots, especially the reduction of very small "dots" which attracted no attention in the past.

Another disadvantage of the conventional light receiving member for electrophotography is its low mechanical strength. When it comes into contact with foreign matters which have entered the electrophotographic apparatus, or when it comes into contact with the main body or tools while the electrophotographic apparatus is being serviced for maintenance, image defects occur or the A-Si film peels off on account of the mechanical shocks and pressure. These aggravate the durability of the light receiving member for electrophotography.

An additional disadvantage of the conventional light receiving member for electrophotography is that the A-Si film is susceptible to cracking and peeling on account of the stress which occurs because the A-Si film differs from the aluminum support in the coefficient of thermal expansion. This leads to lower yields in production.

Under the circumstances mentioned above, it is necessary to solve the above-mentioned problems and to improve the light receiving member for electrophotography from the standpoint of its structure as well as the characteristic properties of the A-Si material per se.

**SUMMARY OF THE INVENTION**

It is an object of the present invention to provide a light receiving member for electrophotography which meets the above-mentioned requirements and eliminates the above-mentioned disadvantages involved in the conventional light receiving member.

According to the present invention, the improved light receiving member for electrophotography is made up of an aluminum support and a multilayered light receiving layer exhibiting photoconductivity formed on the aluminum support, wherein the multilayered light receiving layer consists of a lower layer in contact with the support and an upper layer, the lower layer being made of an inorganic material containing at least aluminum atoms (Al), silicon atoms (Si), and hydrogen atoms (H) ("AlSiH" for short hereinafter), and having a portion in which the aluminum atoms (Al), silicon atoms (Si), and hydrogen atoms (H) are unevenly distributed across the layer thickness, the upper layer being made of a non-single-crystal material composed of silicon

atoms (Si) as the matrix and at least either of hydrogen atoms (H) or halogen atoms (X) ("Non-Si (H,X): for short hereinafter), and containing atoms (M) to control the conductivity in the layer region in adjacent with the lower layer.

The light receiving member for electrophotography in the present invention has the multilayered structure as mentioned above. Therefore, it is free from the above-mentioned disadvantages, and it exhibits outstanding electric characteristics, optical characteristics, photoconductive characteristics, durability, image characteristics, and adaptability to ambient environments.

As mentioned above, the lower layer is made such that the aluminum atoms and silicon atoms, and especially the hydrogen atoms, are unevenly distributed across the layer thickness. This structure improves the injection of electric charge (photocarrier) across the aluminum support and the upper layer. In addition, this structure joins the constituent elements of the aluminum support to the constituent elements of the upper layer gradually in terms of composition and constitution. This leads to the improvement of image characteristics relating to coarse image and dots. Therefore, the light receiving member permits the stable reproduction of images of high quality with a sharp half tone and a high resolving power.

The above-mentioned multilayered structure prevents the image defects and the peeling of the non-Si(H,X) film which occurs as the result of impactive mechanical pressure applied to the light receiving member for electrophotography. In addition, the multilayered structure relieves the stress arising from the difference between the aluminum support and the non-Si(H,X) film in the coefficient of thermal expansion and also prevents the occurrence of cracks and peeling in the non-Si(H,X) film. All this contributes to improved durability and increased yields in production.

Particularly, since the atoms (M) for controlling the conductivity are incorporated into the layer region of the upper layer in adjacent with the lower layer in this invention, injection of electric charges or inhibiting the injection of the charges across the upper layer and the lower layer can selectively be controlled or improved, whereby image property such as "coarse image" or "dots" can further be improved, thereby enabling stable reproduction of high quality images with a clear half-tone and high resolving power, as well as improving charging power, sensitivity and durability.

According to the present invention, the lower layer of the light receiving member may further contain atoms to control the image ("atoms (Mc)" for short hereinafter). The incorporation of atoms (Mc) to control the image quality improves the injection of electric charge (photocarrier) across the aluminum support and the upper layer and also improves the transferability of electric charge (photocarrier) in the lower layer. Thus the light receiving member permits the stable reproduction of images of high quality with a sharp half tone and a high resolving power.

According to the present invention, the lower layer of the light receiving member may further contain atoms to control the durability ("atoms (CNOc)" for short hereinafter). The incorporation of atoms (CNOc) greatly improves the resistance to impactive mechanical pressure applied to the light receiving member for electrophotography. In addition, it prevents the image defects and the peeling of the non-Si(H,X) film, relieves

the stress arising from the difference between the aluminum support and the non-Si(H,X) film in the coefficient of thermal expansion, and prevents the occurrence of cracks and peeling in the non-Si(H,X) film. All this contributes to improved durability and increased yields in production.

According to the present invention, the lower layer of the light receiving member may further contain halogen atom (X). The incorporation of halogen atom (X) compensates for the dangling bonds of silicon atom (Si) and aluminum atom (Al), thereby creating a stable state in terms of constitution and structure. This, coupled with the effect produced by the distribution of silicon atoms (Si), aluminum atoms (Al), and hydrogen atoms (H) mentioned above, greatly improves the image characteristics relating to coarse image and dots.

According to the present invention, the lower layer of the light receiving member may further contain at least either of germanium atoms (Ge) or tin atoms (Sn). The incorporation of at least either of germanium atoms (Ge) or tin atoms (Sn) improves the injection of electric charge (photocarrier) across the aluminum support and the upper layer, the adhesion of the lower layer to the aluminum support, and the transferability of electric charge (photocarrier) in the lower layer. This leads to a distinct improvement in image characteristics and durability.

According to the present invention, the lower layer of the light receiving member may further contain at least one kind of atoms selected from alkali metal atoms, alkaline earth metal atoms, and transition metal atoms, ("atoms (Me)" for short hereinafter). The incorporation of at least one kind of atoms selected from alkali metal atoms, alkaline earth metal atoms, and transition metal atoms permits more dispersion of the hydrogen atoms or halogen atoms contained in the lower layer (the reason for this is not yet fully elucidated) and also reduces the structure relaxation of the lower layer which occurs with lapse of time. This leads to reduced liability of cracking and peeling even after use for a long period of time. The incorporation of at least one kind of the above-mentioned metal atoms improves the injection of electric charge (photocarrier) across the aluminum support and the upper layer, the adhesion of the lower layer to the aluminum support, and the transferability of electric charge (photocarrier) in the lower layer. This leads to a distinct improvement in image characteristics and durability, which in turn leads to the stable production and quality.

In the meantime, the above-mentioned Japanese Patent Laid-open No. 28162/1984 mentions the layer containing aluminum atoms and silicon atoms unevenly across the layer thickness and also mentions the layer containing hydrogen atoms. However, it does not mention how the layer contains hydrogen atoms. Therefore, it is distinctly different from the present invention.

#### BRIEF DESCRIPTION OF THE INVENTION

FIG. 1 is a schematic diagram illustrating the layer structure of the light receiving member for electrophotography.

FIG. 2 is a schematic diagram illustrating the layer structure of the conventional light receiving member for electrophotography.

FIGS. 3 to 8 are diagrams illustrating the distribution state of aluminum atoms (Al) contained in the lower layer, and also illustrating the distribution of atoms (Mc) to control image quality, and/or atoms (CNOc) to

control durability, and/or halogen atoms (X), and/or germanium atoms (Ge), and/or tin atoms (Sn), and/or at least one kind of atoms selected from alkali metal atoms, alkaline earth metal atoms, and transition metal atoms, which are optionally contained in the lower layer.

FIGS. 9 to 16 are diagrams illustrating the distribution of silicon atoms (Si) and hydrogen atoms (H) contained in the lower layer, and also illustrating the distribution of atoms (Mc) to control image quality, and/or atoms (CNOc) to control durability, and/or halogen atoms (X), and/or germanium atoms (Ge), and/or tin atoms (Sn), and/or at least one kind of atoms selected from alkali metal atoms, alkaline earth metal atoms, and transition metal atoms, which are optionally contained in the lower layer.

FIGS. 17 to 36 are diagrams illustrating the distribution of atoms (M) to control conductivity, carbon atoms (C), and/or nitrogen atoms (N), and/or oxygen atoms (O), and/or germanium atoms (Ge), and/or tin atoms (Sn), and/or alkali metal atoms, and/or alkaline earth metal atoms, and/or transition metal atoms, which are contained in the upper layer.

FIG. 37 is a schematic diagram illustrating an apparatus to form the light receiving layer of the light receiving member for electrophotography by RF glow discharge method according to the present invention.

FIG. 38 is an enlarged sectional view of the aluminum support having a V-shape rugged surface which is used to form the light receiving member for electrophotography according to the present invention.

FIG. 39 is an enlarged sectional view of the aluminum support having a dimpled surface on which is used to form the light receiving member for electrophotography according to the present invention.

FIG. 40 is a schematic diagram of the depositing apparatus to form the light receiving layer of the light receiving member for electrophotography by microwave glow discharge method according to the present invention.

FIG. 41 is a schematic diagram of the apparatus to form the light receiving layer of the light receiving member for electrophotography by microwave glow discharge method according to the present invention.

FIG. 42 is a schematic diagram of the apparatus to form the light receiving layer of the light receiving member for electrophotography by RF sputtering method according to the present invention.

FIGS. 43(a) to 43(d) show the distribution of the content of the atoms across the layer thickness in Example 232, Comparative Example 8, Example 239, and Example 240, respectively, of the present invention.

#### DETAILED DESCRIPTION OF THE INVENTION

The light receiving member for electrophotography pertaining to the present invention will be described in more detail with reference to the drawings.

FIG. 1 is a schematic diagram showing a typical example of the layer structure suitable for the light receiving member for electrophotography pertaining to the present invention.

The light receiving member 100 for electrophotography as shown in FIG. 1 comprises an aluminum support 101 for use in the light receiving member for electrophotography and, disposed thereon, the light receiving layer 102 having a layered structure comprising a lower layer 103 constituted with AlSiH and having a part in

which the above-mentioned aluminum atoms and silicon atoms are unevenly distributed across the layer thickness and the upper layer 104 constituted with non-Si(H,X) and containing atoms (M) for controlling the conductivity in the layer region in adjacent with the lower layer. Support

The aluminum support 101 used in the present invention is made of an aluminum alloy. The aluminum alloy is not specifically limited in base aluminum and alloy components. The kind and composition of the components may be selected as desired. Therefore, the aluminum alloy used in the present invention may be selected from pure aluminum, Al-Cu alloy, Al-Mn alloy, Al-Mg alloy, Al-Mg-Si alloy, Al-Zn-Mg alloy, Al-Cu-Mg alloy (duralumin and super duralumin), Al-Cu-Si alloy (lauatal), Al-Cu-Ni-Mg alloy (Y-alloy and RR alloy), and aluminum powder sintered body (SAP) which are standardized or registered as a malleable material, castable material, or die casting material in the Japanese Industrial Standards (JIS), AA Standards, BS Standards, DIN Standards, and International Alloy Registration.

The composition of the aluminum alloy used in the invention is exemplified in the following. The scope of the invention is not restricted to the examples.

Pure aluminum conforming to JIS-1100 which is composed of less than 1.0 wt % of Si and Fe, 0.05-0.20 wt % of Cu, less than 0.05 wt % of Mn, less than 0.10 wt % of Zn, and more than 99.00 wt % of Al.

Al-Cu-Mg alloy conforming to JIS-2017 which is composed of 0.05-0.20 wt % of Si, less than 0.7 wt % of Fe, 3.5-4.5 wt % of Cu, 0.40-1.0 wt % of Mn, 0.40-0.8 wt % of Mg, less than 0.25 wt % of Zn, and less than 0.10 wt % of Cr, with the remainder being Al.

Al-Mn alloy conforming to JIS-3003 which is composed of less than 0.6 wt % of Si, less than 0.7 wt % of Fe, 0.05-0.20 wt % of Cu, 1.0-1.5 wt % of Mn, and less than 0.10 wt % of Zn, with the remainder being Al.

Al-Si alloy conforming to JIS-4032 which is composed of 11.0-13.5 wt % of Si, less than 1.0 wt % of Fe, 0.50-1.3 wt % of Cu, 0.8-1.3 wt % of Mg, less than 0.25 wt % of Zn, less than 0.10 wt % of Cr, and 0.5-1.3 wt % of Ni, with the remainder being Al.

Al-Mg alloy conforming to JIS-5086 which is composed of less than 0.40 wt % of Si, less than 0.50 wt % of Fe, less than 0.10 wt % of Cu, 0.20-0.7 wt % of Mn, 3.5-4.5 wt % of Mg, less than 0.25 wt % of Zn, 0.05-0.25 wt % of Cr, and less than 0.15 wt % of Ti, with the remainder being Al.

An alloy composed of less than 0.50 wt % of Si, less than 0.25 wt % of Fe, 0.04-0.20 wt % of Cu, 0.01-1.0 wt % of Mn, 0.5-10 wt % of Mg, 0.03-0.25 wt % of Zn, 0.05-0.50 wt % of Cr, 0.05-0.20 wt % of Ti or Tr, and less than 1.0 cc of H<sub>2</sub> per 100 g of Al, with the remainder being Al.

Al alloy composed of less than 0.12 wt % of Si, less than 0.15 wt % of Fe, less than 0.30 wt % of Mn, 0.5-5.5 wt % of Mg, 0.01-1.0 wt % of Zn, less than 0.20 wt % of Cr, and 0.01-0.25 wt % of Zr, with the remainder being Al.

Al-Mg-Si alloy conforming to JIS-6063 which is composed of 0.20-0.6 wt % of Si, less than 0.35 wt % of Fe, less than 0.10 wt % of Cu, less than 0.10 wt % of Mn, 0.45-0.9 wt % of MgO, less than 0.10 wt % of Zn, less than 0.10 wt % of Cr, and less than 0.10 wt % of Ti, with the remainder being Al.

Al-Zn-Mg alloy conforming to JIS-7NO1 which is composed of less than 0.30 wt % of Si, less than 0.35 wt % of Fe, less than 0.20 wt % of Cu, 0.20-0.7 wt % of

Mn, 1.0-2.0 wt % of Mg, 4.0-5.0 wt % of Zn, less than 0.30 wt % of Cr, less than 0.20 wt % of Ti, less than 0.25 wt % of Zr, and less than 0.10 wt % of V, with the remainder being Al.

In this invention, an aluminum alloy of proper composition should be selected in consideration of mechanical strength, corrosion resistance, workability, heat resistance, and dimensional accuracy which are required according to specific uses. For example, where precision working with mirror finish is required, an aluminum alloy containing magnesium and/or copper together is desirable because of its free-cutting performance.

According to the present invention, the aluminum support 101 can be in the form of cylinder or flat endless belt with a smooth or irregular surface. The thickness of the support should be properly determined so that the light receiving member for electrophotography can be formed as desired. In the case where the light receiving member for electrophotography is required to be flexible, it can be made as thin as possible within limits not harmful to the performance of the support. Usually the thickness should be greater than 10  $\mu$ m for the convenience of production and handling and for the reason of mechanical strength.

In the case where the image recording is accomplished by the aid of coherent light such as laser light, the aluminum support may be provided with an irregular surface to eliminate defective images caused by interference fringes.

The irregular surface on the support may be produced by any known method disclosed in Japanese Patent Laid-open Nos. 168156/1985, 178457/1985, and 225854/1985.

The support may also be provided with an irregular surface composed of a plurality of spherical dents in order to eliminate defective images caused by interference fringes which occur when coherent light such as laser light is used.

In this case, the surface of the support has irregularities smaller than the resolving power required for the light receiving member for electrophotography, and the irregularities are composed of a plurality of dents.

The irregularities composed of a plurality of spherical dents can be formed on the surface of the support according to the known method disclosed in Japanese Patent Laid-open No. 231561/1986.

#### Lower layer

According to the present invention, the lower layer is made of an inorganic material which is composed of at least aluminum atoms (Al), silicon atoms (Si), and hydrogen atoms (H). It may further contain atoms (Mc) to control image quality, atoms (CNOc) to control durability, halogen atoms (X), germanium atoms (Ge), and/or tin atoms (Sn), and at least one kind of atoms (Me) selected from the group consisting of alkali metal atoms, and/or alkaline earth metal atoms, and transition metal atoms.

The lower layer contains aluminum atoms (Al), silicon atoms, (Si), and hydrogen atoms (H) which are distributed evenly throughout the layer; but it has a part in which their distribution is uneven across the layer thickness. Their distribution should be uniform in a plane parallel to the surface of the support so that uniform characteristics are ensured in the same plane.

According to a preferred embodiment, the lower layer contains aluminum atoms (Al), silicon atoms (Si),

and hydrogen atoms (H) which are distributed evenly and continuously throughout the layer, with the aluminum atoms (Al) being distributed such that their concentration gradually decreases across the layer thickness toward the upper layer from the support, with the silicon atoms (Si) and hydrogen atoms (H) being distributed such that their concentration gradually increases across the layer thickness toward the upper layer from the support. This distribution of atoms makes the aluminum support and the lower layer compatible with each other and also makes the lower layer and the upper layer compatible with each other.

In the light receiving member for electrophotography according to the present invention, it is desirable that the lower layer contains aluminum atoms (Al), silicon atoms (Si), and hydrogen atoms (H) which are specifically distributed across the layer thickness as mentioned above but are evenly distributed in the plane parallel to the surface of the support.

15 The lower layer may further contain atoms (Mc) to control image quality, atoms (CNOc) to control durability, halogen atoms (X), germanium atoms (Ge), and/or tin atoms (Sn), and at least one kind of atoms (Me) selected from the group consisting of alkali metal atoms,

25 alkaline earth metal atoms, and transition metal atoms, which are evenly distributed throughout the entire layer or unevenly distributed across the layer thickness in a specific part. In either case, their distribution should be uniform in a plane parallel to the surface of the support so that uniform characteristics are ensured in the same plane.

30 FIGS. 3 to 8 show the typical examples of the distribution of aluminum atoms (Al) and optionally added atoms in the lower layer of the light receiving member for electrophotography in the present invention. (The aluminum atoms (Al) and the optionally added atoms are collectively referred to as "atoms (AM)" hereinafter.)

35 In FIGS. 3 to 8, the abscissa represents the concentration (C) of atoms (AM) and the ordinate represents the thickness of the lower layer. (The aluminum atoms (Al) and the optionally added atoms may be the same or different in their distribution across the layer thickness.)

40 The ordinate represents the thickness of the lower layer, with  $t_B$  representing the position of the end (adjacent to the support) of the lower layer, with  $t_T$  representing the position of the end (adjacent to the upper layer) of the lower layer. In other words, the lower layer containing atoms (AM) is formed from the  $t_B$  side toward the  $t_T$  side.

45 FIG. 3 shows a first typical example of the distribution of atoms (AM) across layer thickness in the lower layer. The distribution shown in FIG. 3 is such that the concentration (C) of atoms (AM) remains constant at  $C_{31}$  between position  $t_B$  and position  $t_{31}$  and linearly decreases from  $C_{31}$  to  $C_{32}$  between position  $t_{31}$  and position  $t_T$ .

50 The distribution shown in FIG. 4 is such that the concentration (C) of atoms (AM) linearly decreases from  $C_{41}$  to  $C_{42}$  between position  $t_B$  and position  $t_T$ .

The distribution shown in FIG. 5 is such that the concentration (C) of atoms (AM) gradually and continuously decreases from  $C_{51}$  to  $C_{52}$  between position  $t_B$  and position  $t_T$ .

55 The distribution shown in FIG. 6 is such that the concentration (C) of atoms (AM) remains constant at  $C_{61}$  between position  $t_B$  and position  $t_{61}$  and linearly decreases from  $C_{62}$  to  $C_{63}$  between  $t_{61}$  and position  $t_T$ .

The distribution shown in FIG. 7 is such that the concentration (C) of atoms (AM) remains constant at  $C_{71}$  between position  $t_B$  and position  $t_{71}$  and decreases gradually and continuously from  $C_{72}$  to  $C_{73}$  between position  $t_{71}$  and position  $t_T$ .

The distribution shown in FIG. 8 is such that the concentration (C) of atoms (AM) decreases gradually and continuously from  $C_{81}$  to  $C_{82}$  between position  $t_B$  and position  $t_T$ .

The atoms (AM) in the lower layer are distributed across the layer thickness as shown in FIGS. 3 to 8 with reference to several typical examples. In a preferred embodiment, the lower layer contains silicon atoms (Si) and hydrogen atoms (H) and atoms (AM) in a high concentration of C in the part adjacent to the support, and also contains atoms (AM) in a much lower concentration at the interface  $t_T$ . In such a case, the distribution across the layer thickness should be made such that the maximum concentration  $C_{max}$  of atoms (Al) is 10 atom %, or above, preferably 30 atom % or above, and most desirably 50 atom % or above.

According to the present invention, the amount of atoms (Al) in the lower layer should be properly established so that the object of the invention is effectively achieved. It is 5-95 atom %, preferably 10-90 atom %, and most desirably 20-80 atom %.

FIGS. 9 to 16 shows the typical examples of the distribution of silicon atoms (Si), hydrogen atoms (H), and the above-mentioned optional atoms contained across the layer thickness in the lower layer of the light receiving member for electrophotography in the present invention.

In FIGS. 9 to 16, the abscissa represents the concentration (C) of silicon atoms (Si), hydrogen atoms (H), and optionally contained atoms and the ordinate represents the thickness of the lower layer will be collectively referred to as "atoms (SHM)" hereinafter.) The silicon atoms (Si), hydrogen atoms (H), and optionally contained atoms may be the same or different in their distribution across the layer thickness.  $t_B$  on the ordinate represents the end of the lower layer adjacent to the support and  $t_T$  on the ordinate represents the end of the lower layer adjacent to the upper layer. In other words, the lower layer containing atoms (SHM) is formed from the  $t_B$  side toward the  $t_T$  side.

FIG. 9 shows a first typical example of the distribution of atoms (SHM) across the layer thickness in the lower layer. The distribution shown in FIG. 9 is such that the concentration (C) of atoms (SHM) linearly increases from  $C_{91}$  to  $C_{92}$  between position  $t_B$  and position  $t_{91}$  and remains constant at  $C_{92}$  between position  $t_{91}$  and position  $t_T$ .

The distribution shown in FIG. 10 is such that the concentration (C) of atoms (SHM) linearly increases from  $C_{101}$  to  $C_{102}$  between position  $t_B$  and position  $t_T$ .

The distribution shown in FIG. 11 is such that the concentration (C) of atoms (SHM) gradually and continuously increase from  $C_{111}$  to  $C_{112}$  between position  $t_B$  and position  $t_T$ .

The distribution shown in FIG. 12 is such that the concentration (C) of atoms (SHM) linearly increases from  $C_{121}$  to  $C_{122}$  between position  $t_B$  and position  $t_{121}$  and remains constant at  $C_{123}$  between position  $t_{121}$  and position  $t_T$ .

The distribution shown in FIG. 13 is such that the concentration (C) of atoms (SHM) gradually and continuously increases from  $C_{131}$  to  $C_{132}$  between position

$t_B$  and position  $t_{131}$  and remains constant at  $C_{133}$  between position  $t_{131}$  and position  $t_T$ .

The distribution shown in FIG. 14 is such that the concentration (C) of atoms (SHM) gradually and continuously increases from  $C_{141}$  to  $C_{142}$  between position  $t_B$  and position  $t_T$ .

The distribution shown in FIG. 15 is such that the concentration (C) of atoms (SHM) gradually increases from substantially zero to  $C_{151}$  between position  $t_B$  and position  $t_{151}$  and remains constant at  $C_{152}$  between position  $t_{151}$  and position  $t_T$ . ("Substantially zero" means that the amount is lower than the detection limit. The same shall apply hereinafter.)

The distribution shown in FIG. 16 is such that the concentration (C) of atoms (SHM) gradually increases from substantially zero to  $C_{161}$  between position  $t_B$  and position  $t_T$ .

The silicon atoms (Si) and hydrogen atoms (H) in the lower layer are distributed across the layer thickness as shown in FIGS. 9 to 16 with reference to several typical examples. In a preferred embodiment, the lower layer contains aluminum atoms (Al) and silicon atoms (Si) and hydrogen atoms (H) in a low concentration of C in the part adjacent to the support, and also contains silicon atoms (Si) and hydrogen atoms (H) in a much higher concentration at the interface  $t_T$ . In such a case, the distribution across the layer thickness should be made such that the maximum concentration  $C_{max}$  of the total of silicon atoms (Si) and hydrogen atoms (H) is 10 atom % or above, preferably 30 atom % or above, preferably 30 atom % or above, and most desirably 50 atom % or above.

According to the present invention, the amount of silicon atoms (Si) in the lower layer should be properly established so that the object of the invention is effectively achieved. It is 5-95 atom %, preferably 10-90 atom %, and most desirably 20-80 atom %.

According to the present invention, the amount of hydrogen atoms (H) in the lower layer should be properly established so that the object of the invention is effectively achieved. It is 0.01-70 atom %, preferably 0.1-50 atom %, and most desirably 1-40 atom %.

The above-mentioned atoms (Mc) optionally contained to control image quality are selected from atoms belonging to Group III of the periodic table, except for aluminum atoms (Al) ("Group III atoms" for short hereinafter), atoms belonging to Group V of the periodic table, except for nitrogen atoms (N) ("Group V atoms" for short hereinafter), and atoms belonging to Group VI of the periodic table, except for oxygen atoms (O) ("Group VI atoms" for short hereinafter).

Examples of Group III atoms include B (boron), Ga (gallium), In (indium), and Tl (thallium), with B, Al and Ga being preferable. Examples of Group V atoms include P (phosphorus), As (arsenic), Sb (antimony) and Bi (bismuth), with P and As being preferable. Examples of Group VI atoms include S (sulfur), Se (selenium), Te (tellurium), and Po (polonium), with S and Se being preferable.

According to the present invention, the lower layer may contain atoms (Mc) to control image quality, which are Group III atoms, Group V atoms, or Group VI atoms. The atoms (Mc) improve the injection of electric charge across the aluminum support and the upper layer and/or improve the transferability of electric charge in the lower layer. They also control conduction type and/or conductivity in the region of the

lower layer which contains a less amount of aluminum atoms (Al).

In the lower layer, the content of atoms (Mc) to control image quality should be  $1 \times 10^{-3}$ – $5 \times 10^4$  atom-ppm, preferably  $1 \times 10^{-1}$ – $5 \times 10^4$  atom-ppm, and most desirably  $1 \times 10^{-2}$ – $5 \times 10^3$  atom-ppm.

The above-mentioned atoms (NCOc) optionally contained to control durability are selected from carbon atoms (C), nitrogen atoms (N), and oxygen atoms (O). When contained in the lower layer, carbon atoms (C), and/or nitrogen atoms (N), and/or oxygen atoms (O) as the atoms (CNOc) to control durability improve the injection of electric charge across the aluminum support and the upper layer and/or improve the transferability of electric charge in the lower layer and/or improve the adhesion of the lower layer to the aluminum support. They also control the width of the forbidden band in the region of the lower layer which contains a less amount of aluminum atoms (Al).

In the lower layer, the content of atoms (NCOc) to control durability should be  $1 \times 10^3$ – $5 \times 10^5$  atom-ppm, preferably  $5 \times 10^1$ – $4 \times 10^5$  atom-ppm, and most desirably  $1 \times 10^2$ – $3 \times 10^3$  atom-ppm.

The above-mentioned halogen atoms (X) optionally contained in the lower layer are selected from fluorine atoms (F), chlorine atoms (Cl), bromine atoms (Br), and iodine atoms (I). When contained in the lower layer, fluorine atoms (F), and/or chlorine atoms (Cl), and/or bromine atoms (Br), and/or iodine atoms (I) as the halogen atoms (V) compensate for the unbonded hands of silicon atoms (Si) and aluminum atoms (Al) contained mainly in the lower layer and make the lower layer stable in terms of composition and structure, thereby improving the quality of the layer.

The content of halogen atoms (X) in the lower layer should be properly established so that the object of the invention is effectively achieved. It is  $1$ – $4 \times 10^5$  atom-ppm, preferably  $10$ – $3 \times 10^5$  atom-ppm, and most desirably  $1 \times 10^2$ – $2 \times 10^5$  atom-ppm.

According to the present invention, the lower layer may optionally contain germanium atoms (Ge) and/or tin atoms (Sn). They improve the injection of electric charge across the aluminum support and the upper layer and/or improve the transferability of electric charge in the lower layer and/or improve the adhesion of the lower layer to the aluminum support. They also narrow the width of the forbidden band in the region of the lower layer which contains a less amount of aluminum atoms (Al). These effects suppress interference which occurs when a light of long wavelength such as semiconductor laser is used as the light source for image exposure in the electrophotographic apparatus.

The content of germanium atoms (Ge) and/or tin atoms (Sn) in the lower layer should be properly established so that the object of the invention is effectively achieved. It is  $1$ – $9 \times 10^5$  atom-ppm, preferably  $1 \times 10^2$ – $8 \times 10^5$  atom-ppm, and most desirably  $5 \times 10^2$ – $7 \times 10^5$  atom-ppm.

According to the present invention, the lower layer may optionally contain, as the alkali metal atoms and/or alkaline earth metal atoms and/or transition metal atoms, magnesium atoms (Mg) and/or copper atoms (Cu) and/or sodium atoms (Na) and/or yttrium atoms (Y) and/or manganese atoms (Mn) and/or zinc atoms (Zn). They disperse hydrogen atoms (H) and halogen atoms (X) uniformly in the lower layer and prevent the cohesion of hydrogen which is considered to cause cracking and peeling. They also improve the injection

of electric charge across the aluminum support and the upper layer and/or improve the transferability of electric charge in the lower layer and/or improve the adhesion of the lower layer to the aluminum support.

The content of the above-mentioned metals in the lower layer should be properly established so that the object of the invention is effectively achieved. It is  $1$ – $2 \times 10^5$  atom-ppm, preferably  $1 \times 10^2$ – $1 \times 10^5$  atom-ppm, and most desirably  $5 \times 10^2$ – $5 \times 10^4$  atom-ppm.

According to the present invention, the lower layer composed of AlSiH is formed by the vacuum deposition film forming method, as in the upper layer which will be mentioned later, under proper conditions for the desired characteristic properties. The thin film is

15 formed by one of the following various methods. Glow discharge method (including ac current discharge CVD, e.g., low-frequency CVD, high-frequency CVD, and microwave CVD, and dc current CVD), ECR-CVD method, sputtering method, vacuum metallizing method, ion plating method, light CVD method, "HRCVD" method (explained below), "FOCVD" method (explained below). (According to HRCVD method, an active substance (A) formed by the decomposition of a raw material gas and the other active substance (B) formed from a substance reactive to the first active substance are caused to react with each other in a space where the film formation is accomplished. According to FOCVD method, a raw material gas and a halogen-derived gas capable of oxidizing said raw material gas are caused to react in a space where the film formation is accomplished.) A proper method should be selected according to the manufacturing conditions, the capital available, the production scale, and the characteristic properties required for the light receiving member for electrophotography. Preferable among these methods are glow discharge method, sputtering method, ion plating method, HRCVD method, and FOCVD method on account of their ability to control the production conditions and to introduce aluminum atoms (Al), silicon atoms (Si), and hydrogen atoms (H) with ease. These methods may be used in combination with one another in the same apparatus.

The glow discharge method may be performed in the following manner to form the lower layer of AlSiH. 45 The raw material gases are introduced into an evacuable deposition chamber, and glow discharge is performed, with the gases being introduced at a desired pressure, so that a layer of AlSiH is formed as required on the surface of the support placed in the chamber. 50 The raw material gases may contain a gas to supply aluminum atoms (Al), a gas to supply silicon atoms (Si), a gas to supply hydrogen atoms (H), an optional gas to supply atoms (Mc) to control image quality, an optional gas to supply atoms (CNOx) to control durability, an optional gas to supply halogen atoms (X), an optional gas to supply atoms (GSc) (germanium atoms (Ge) and tin atoms (Sn), and an optional gas to supply atoms (Me) (at least one kind of alkali metal atoms, alkaline earth metal atoms, and transition metal atoms).

60 The HRCVD may be performed in the following manner to form the lower layer of AlSiH. The raw material gases are introduced all together or individually into an evacuable deposition chamber, and glow discharge is performed or the gases are heated, with the gases being introduced at a desired pressure, during which a first active substance (A) is formed and a second active substance (B) is introduced into the deposition chamber, so that a layer of AlSiH is formed as

required on the surface of the support placed in the chamber. The raw material gases may contain a gas to supply aluminum atoms, (Al), a gas to supply silicon atoms (Si), an optional gas to supply atoms (Mc) to control image quality, an optional gas to supply atoms (CNOc) to control durability, an optional gas to supply halogen atoms (X), an optional gas to supply atoms (GSc) (germanium atoms (Ge) and tin atoms (Sn)), and an optional gas to supply atoms (Me) (at least one kind of alkali metal atoms, alkaline earth metal atoms, and transition metal atoms). A second active substance (B) is formed by introducing a gas to supply hydrogen into the activation chamber. Said first active substance (A) and said second active substance are individually introduced into the deposition chamber.

The FOCVD method may be performed in the following manner to form the lower layer of AlSiH. The raw material gases are introduced into an evacuable deposition chamber, and chemical reactions are performed, with the gases being introduced at a desired pressure, so that a layer of AlSiH is formed as required on the surface of the support placed in the chamber. The raw material gases may contain a gas to supply aluminum atoms (Al), a gas to supply silicon atoms (Si), a gas to supply hydrogen atoms (H), an optional gas to supply atoms (Mc) to control image quality, an optional gas to supply atoms (CNOc) to control durability, an optional gas to supply halogen atoms (X), an optional gas to supply atoms (GSc) (germanium atoms (Ge) and tin atoms (Sn)), and an optional gas to supply atoms (Me) (at least one kind of alkali metal atoms, alkaline earth metal atoms, and transition metal atoms). They may be introduced into the chamber altogether or individually, and a halogen (X) gas is introduced into the chamber separately from said raw materials gas, and these gases are subjected to chemical reaction in the deposition chamber.

The sputtering method may be performed in the following manner to form the lower layer of AlSiH. The raw material gases are introduced into a sputtering deposition chamber, and a desired gas plasma environment is formed using an aluminum target and an Si target in an inert gas of Ar or He or an Ar- or He-containing gas. The raw material gases may contain a gas to supply hydrogen atoms (H), an optional gas to supply atoms (Mc) to control image quality, an optional gas to supply atoms (CNOc) to control durability, an optional gas to supply halogen atoms (X), an optional gas to supply atoms (GSc) (Germanium atoms (Ge) and tin atoms (Sn)), and an optional gas to supply atoms (Me) (at least one kind of alkali metal atoms, alkaline earth metal atoms, and transition metal atoms). If necessary, a gas to supply aluminum atoms (Al) and/or to supply silicon atoms (Si) are introduced into the sputtering chamber.

The ion plating method may be performed in the same manner as the sputtering method, except that vapors of aluminum and silicon are passed through the gas plasma environment. The vapors of aluminum and silicon are produced from aluminum and silicon polycrystal or single crystal placed in a boat which is heated by resistance or electron beams (EB method).

According to the present invention, the lower layer contains aluminum atoms (Al), silicon atoms (Si), hydrogen atoms (H), optional atoms (Mc) to control image quality, optional atoms (CNOc) to control durability, optional halogen atoms (X), optional germanium atoms (Ge), optional tin atoms (Sn), optional alkali metal

atoms, optional alkaline earth metal atoms, and optional transition metal atoms (collectively referred to as atoms (ASH) hereinafter), which are distributed in different concentrations across the layer thickness. The lower layer having such a depth profile can be formed by controlling the flow rate of the feed gas to supply atoms (ASH) according to the desired rate of change in concentration. The flow rate may be changed by operating the needle valve in the gas passage manually or by means of a motor, or it may be changed by any of customary means such as by properly adjusting the mass flow controller manually or by means of a programmable control apparatus.

In the case where the sputtering method is used, the lower layer having such a depth profile can be formed, as in the glow discharge method, it can be achieved by controlling the flow rate of the gaseous raw material to supply atoms (ASH) according to the desired rate of change in concentration and introducing the gas into the deposition chamber. Alternatively, it is possible to use a sputtering target comprising a Al-Si mixture in which the mixing ratio of Al and Si is properly changed in the direction of layer thickness of the target.

According to the present invention, the gas to supply Al includes, for example, AlCl<sub>3</sub>, AlBr<sub>3</sub>, AlI<sub>3</sub>, Al(CH<sub>3</sub>)<sub>2</sub>Cl, Al(CH<sub>3</sub>)<sub>2</sub>, Al(OCH<sub>3</sub>)<sub>3</sub>, Al(C<sub>2</sub>H<sub>5</sub>)<sub>3</sub>, Al(i-C<sub>4</sub>H<sub>9</sub>)<sub>3</sub>, Al(i-C<sub>3</sub>H<sub>7</sub>)<sub>3</sub>, Al(C<sub>3</sub>H<sub>7</sub>)<sub>3</sub> and (Al(OC<sub>4</sub>H<sub>9</sub>)<sub>3</sub>). These gases to supply Al may be diluted with an inert gas such as H<sub>2</sub>, He, Ar and Ne, if necessary.

According to the present invention, the gas to supply Si includes, for example, gaseous or gasifiable silicohydrides (silanes) such as SiH<sub>4</sub>, Si<sub>2</sub>H<sub>6</sub>, Si<sub>3</sub>H<sub>8</sub> and Si<sub>4</sub>H<sub>10</sub>. SiH<sub>4</sub> and Si<sub>2</sub>H<sub>6</sub> are preferable from the standpoint of each of handling and the efficient supply of Si. These gases to supply Si may be diluted with an inert gas such as H<sub>2</sub>, He, Ar and Ne, if necessary.

According to the present invention, the gas to supply H includes, for example, silicohydrides (silanes) such as SiH<sub>4</sub>, Si<sub>2</sub>H<sub>6</sub>, Si<sub>3</sub>H<sub>8</sub> and Si<sub>4</sub>H<sub>10</sub>.

The amount of hydrogen atoms contained in the lower layer may be controlled by regulating the flow rate of the feed gas to supply hydrogen and/or regulating the temperature of the support and/or regulating the electric power for discharge.

The lower layer may contain atoms (Mc) to control image quality, such as Group III atoms, Group V atoms and Group VI atoms. This is accomplished by introducing into the deposition chamber the raw materials to form the lower layer together with a raw material to introduce Group III atoms, a raw material to introduce Group V atoms, or a raw material to introduce Group VI atoms. The raw material to introduce Group III atoms, the raw material to introduce Group V atoms, or the raw material to introduce Group VI atoms may desirably be gaseous at normal temperature and under normal pressure or gasifiable under the layer forming conditions. The raw material to introduce Group III atoms, especially boron atoms, include, for example, boron, hydrides such as B<sub>2</sub>H<sub>6</sub>, B<sub>5</sub>H<sub>9</sub>, B<sub>5</sub>H<sub>11</sub>, B<sub>6</sub>H<sub>10</sub>, B<sub>6</sub>H<sub>12</sub> and B<sub>6</sub>H<sub>14</sub>, and boron halides such as BF<sub>3</sub>, BCl<sub>3</sub> and BBr<sub>3</sub>. Additional examples includes GaCl<sub>3</sub>, Ga(CH<sub>3</sub>)<sub>3</sub>, InCl<sub>3</sub> and TiCl<sub>3</sub>.

The raw material to introduce Group V atoms, especially phosphorus atoms, include, for example, phosphorus hydrides such as PH<sub>3</sub>, P<sub>2</sub>H<sub>4</sub> and phosphorus halides such as PH<sub>4</sub>I, PF<sub>3</sub>, PF<sub>5</sub>, PCl<sub>3</sub>, PBr<sub>3</sub>, PBr<sub>5</sub> and PI<sub>3</sub>. Other examples effective to introduce Group V

atoms include  $\text{AsH}_3$ ,  $\text{AsF}_3$ ,  $\text{AsCl}_3$ ,  $\text{AsBr}_3$ ,  $\text{AsF}_5$ ,  $\text{SbH}_3$ ,  $\text{SbF}_3$ ,  $\text{SbF}_5$ ,  $\text{SbCl}_3$ ,  $\text{SbCl}_5$ ,  $\text{BiH}_3$ ,  $\text{BiCl}_3$  and  $\text{BiBr}_3$ .

The raw material to introduce Group VI atoms includes, for example, gaseous or gasifiable substances such as  $\text{H}_2$ ,  $\text{SF}_4$ ,  $\text{SF}_6$ ,  $\text{SO}_2$ ,  $\text{SO}_2\text{F}_2$ ,  $\text{COS}$ ,  $\text{CS}_2$ ,  $\text{CH}_3\text{SH}$ ,  $\text{C}_2\text{H}_5\text{SH}$ ,  $\text{C}_4\text{H}_4\text{S}$ ,  $(\text{CH}_3)_2\text{S}$  and  $\text{S}(\text{C}_2\text{H}_5)_2\text{S}$ . Other examples include gaseous or gasifiable substances such as  $\text{SeH}_2$ ,  $\text{SeF}_6$ ,  $(\text{CH}_3)_2\text{Se}$ ,  $(\text{C}_2\text{H}_5)_2\text{Se}$ ,  $\text{TeH}_2$ ,  $\text{TeF}_6$ ,  $(\text{CH}_3)_2\text{Te}$  and  $(\text{C}_2\text{H}_5)_2\text{Te}$ .

These raw materials to introduce atoms (Mc) to control image quality may be diluted with an inert gas such as  $\text{H}_2$ ,  $\text{He}$ ,  $\text{Ar}$  and  $\text{Ne}$ .

According to the present invention, the lower layer may contain atoms (CNOc) to control durability, e.g., carbon atoms (C), nitrogen atom (N), and oxygen atoms (O). This is accomplished by introducing into the deposition chamber the raw materials to form the lower layer, together with a raw material to introduce carbon atoms (C), or a raw material to introduce nitrogen atoms (N), or a raw material to introduce oxygen atoms (O). Raw materials to introduce carbon atoms (C), nitrogen atoms (N), or oxygen atoms (O) may desirably be in the gaseous form at normal temperature and under normal pressure or may be readily gasifiable under the layer forming conditions.

A raw material gas to introduce carbon atoms (C) includes those composed of C and H atoms such as saturated hydrocarbons having 1 to 4 carbon atoms, ethylene, series hydrocarbons having 2 to 4 carbon atoms and acetylene series hydrocarbons having 2 to 3 carbon atoms.

Examples of the saturated hydrocarbons include specifically methane ( $\text{CH}_4$ ), ethane ( $\text{C}_2\text{H}_6$ ), propane ( $\text{C}_3\text{H}_8$ ), n-butane ( $n\text{-C}_4\text{H}_{10}$ ) and pentane ( $\text{C}_5\text{H}_{12}$ ). Examples of the ethylene series hydrocarbons include ethylene ( $\text{C}_2\text{H}_4$ ), propylene ( $\text{C}_3\text{H}_6$ ), butene-1 ( $\text{C}_4\text{H}_8$ ), butene-2 ( $\text{C}_4\text{H}_8$ ), isobutylene ( $\text{C}_4\text{H}_8$ ) and pentene ( $\text{C}_5\text{H}_{10}$ ). Examples of acetylene series hydrocarbon include acetylene ( $\text{C}_2\text{H}_2$ ), methylacetylene ( $\text{C}_3\text{H}_4$ ) and butyne ( $\text{C}_4\text{H}_6$ ).

The raw material gas composed of Si, C, and H includes alkyl silicides such as  $\text{Si}(\text{CH}_3)_4$  and  $\text{Si}(\text{C}_2\text{H}_5)_4$ .

Additional examples include gases of halogenated hydrocarbons such as of  $\text{CF}_4$ ,  $\text{CCl}_4$  and  $\text{CH}_3\text{CF}_3$ , which introduce carbon atoms (C) as well as halogen atoms (X).

Examples of the raw material gas to introduce nitrogen atoms (N) include nitrogen and gaseous or gasifiable nitrogen compounds (e.g., nitrides and azides) which are composed of nitrogen and hydrogen, such as ammonia ( $\text{NH}_3$ ), hydrazine ( $\text{H}_2\text{NNH}_2$ ), hydrogen azide ( $\text{HN}_3$ ), and ammonium azide ( $\text{NH}_4\text{N}_3$ ).

Additional examples include halogenated nitrogen compounds such as nitrogen trifluoride ( $\text{F}_3\text{N}$ ) and nitrogen tetrafluoride ( $\text{F}_4\text{N}_2$ ), which can introduce nitrogen atoms as well as halogen atoms (X).

Examples of the raw material gas to introduce oxygen atoms (O) include oxygen ( $\text{O}_2$ ), ozone ( $\text{O}_3$ ), nitrogen monoxide ( $\text{NO}$ ), nitrogen dioxide ( $\text{NO}_2$ ), trinitrogen tetraoxide ( $\text{N}_3\text{O}_4$ ), dinitrogen pentaoxide ( $\text{N}_2\text{O}_5$ ) and nitrogen trioxide ( $\text{NO}_3$ ), as well as lower siloxanes such as disiloxane ( $\text{H}_3\text{SiOSiH}_3$ ) and trisiloxane ( $\text{H}_3\text{SiOSiH}_2\text{OSiH}_3$ ) which are composed of silicon atoms (Si), oxygen atoms (O) and hydrogen atoms (H).

Examples of the gas to supply hydrogen atoms include halogen gases and gaseous or gasifiable halides, interhalogen compounds, and halogen-substituted silane derivatives. Additional examples include gaseous or

gasifiable halogen-containing silicohydrides composed of silicon atoms and halogen atoms.

The halogen compounds that can be suitably used in the present invention include halogen gases such as fluorine, chlorine, bromine and iodine; and interhalogen compounds such as  $\text{BrF}$ ,  $\text{ClF}$ ,  $\text{ClF}_3$ ,  $\text{BrF}_5$ ,  $\text{BrF}_3$ ,  $\text{IF}_3$ ,  $\text{IF}_7$ ,  $\text{ICl}$  and  $\text{IBr}$ .

Examples of the halogen-containing silicon compounds or halogen-substituted silane compounds, include specifically silane ( $\text{SiH}_4$ ) and halogenated silicon such as  $\text{Si}_2\text{F}_6$ ,  $\text{SiCl}_4$  and  $\text{SiBr}_4$ .

In the case where the halogen-containing silicon compounds is used to form the light receiving member for electrophotography by the glow discharge method or HRCVD method, it is possible to form the lower layer composed of  $\text{AlSiH}$  containing halogen atoms on the support without using a silicohydride gas to supply silicon atoms.

In the case where the lower layer containing halogen atoms is formed by the glow discharge method of HRCVD method, a silicon halide gas is used as the gas to supply silicon atoms. The silicon halide gas may be mixed with hydrogen or a hydrogen-containing silicon compound gas to facilitate the introduction of hydrogen atoms at a desired level.

The above-mentioned gases may be used individually or in combination with one another at a desired mixing ratio.

The raw materials to form the lower layer which are used in addition to the above-mentioned halogen compounds or halogen-containing silicon compounds include gaseous or gasifiable hydrogen halides such as  $\text{HF}$ ,  $\text{HCl}$ ,  $\text{HBr}$  and  $\text{HI}$ ; and halogen-substituted silicohydrides such as  $\text{SiH}_3\text{F}_2$ ,  $\text{SiH}_2\text{F}_2$ ,  $\text{SiHF}_3$ ,  $\text{SiH}_2\text{I}_2$ ,  $\text{SiS}_2\text{Cl}_2$ ,  $\text{SiHCl}_3$ ,  $\text{SiH}_2\text{Br}_2$  and  $\text{SiHBr}_3$ . Among these substances, the hydrogen-containing halides are a preferred halogen-supply gas because they supply the lower layer with halogen atoms as well as hydrogen atoms which are very effective for the control of electric or photoelectric characteristics.

The introduction of hydrogen atoms into the lower layer may also be accomplished in another method by inducing discharge in the deposition chamber containing a silicohydride such as  $\text{SiH}_4$ ,  $\text{Si}_2\text{H}_6$ ,  $\text{Si}_3\text{H}_8$  and  $\text{SiK}_4\text{H}_{10}$  and a silicon compound to supply silicon atoms (Si).

The amount of hydrogen atoms (H) and/or halogen atoms (X) to be introduced into the lower layer may be controlled by regulating the temperature of the support, the electric power for discharge, and the amount of raw materials for hydrogen atoms and halogen atoms to be introduced into the deposition chamber.

The lower layer may contain germanium atoms (Ge) or tin atoms (Sn). This is accomplished by introducing into the deposition chamber the raw materials to form the lower layer together with a raw material to introduce germanium atoms (Ge) or tin atoms (Sn) in a gaseous form. The raw material to supply germanium atoms (Ge) or the raw material to supply tin atoms (Sn) may be gaseous at normal temperature and under normal pressure or gasifiable the layer forming conditions.

The substance that can be used as a gas to supply germanium atoms (Ge) include gaseous or gasifiable germanium hydrides such as  $\text{GeH}_4$ ,  $\text{Ge}_2\text{H}_6$ ,  $\text{Ge}_3\text{H}_8$  and  $\text{Ge}_4\text{H}_{10}$ . Among them,  $\text{GeH}_4$ ,  $\text{Ge}_2\text{H}_6$  and  $\text{Ge}_3\text{H}_8$  are preferable from the standpoint of easy handling at the time of layer forming and the efficient supply of germanium atoms (Ge).

Other effective raw materials to form the lower layer include gaseous or gasifiable germanium hydride-halides such as  $\text{GeHF}_3$ ,  $\text{GeH}_2\text{F}_2$ ,  $\text{GeH}_3\text{F}$ ,  $\text{GeHCl}_3$ ,  $\text{GeH}_2\text{Cl}_2$ ,  $\text{GeH}_3\text{Cl}$ ,  $\text{GeHBr}_3$ ,  $\text{GeH}_2\text{Br}_2$ ,  $\text{GeH}_3\text{Br}$ ,  $\text{GeHI}_3$ ,  $\text{GeH}_2\text{I}_2$  and  $\text{GeH}_3\text{I}$  and germanium halides such as  $\text{GeF}_4$ ,  $\text{GeCl}_4$ ,  $\text{GeBr}_4$ ,  $\text{GeI}_4$ ,  $\text{GeF}_2$ ,  $\text{GeCl}_2$ ,  $\text{GeBr}_2$  and  $\text{GeI}_2$ .

The substance that can be used as a gas to supply tin atoms (Sn) include gaseous or gasifiable tin hydrides such as  $\text{SnH}_4$ ,  $\text{Sn}_2\text{H}_6$ ,  $\text{Sn}_3\text{H}_8$  and  $\text{Sn}_4\text{H}_{10}$ . Among them,  $\text{SnH}_4$ ,  $\text{Sn}_2\text{H}_6$  and  $\text{Sn}_3\text{H}_8$  are preferable from the standpoint of easy handling at the time of layer forming and the efficient supply of tin atoms (Sn).

Other effective raw materials to form the lower layer include gaseous or gasifiable tin hydride-halides such as  $\text{SnHF}_3$ ,  $\text{SnH}_2\text{F}_2$ ,  $\text{SnH}_3\text{F}$ ,  $\text{SnHCl}_3$ ,  $\text{SnH}_2\text{Cl}_2$ ,  $\text{SnH}_3\text{Cl}$ ,  $\text{SnHBr}_3$ ,  $\text{SnH}_2\text{Br}_2$ ,  $\text{SnH}_3\text{Br}$ ,  $\text{SnHI}_3$ ,  $\text{SnH}_2\text{I}_2$  and  $\text{SnH}_3\text{I}$ , and tin halides such as  $\text{SnF}_4$ ,  $\text{SnCl}_4$ ,  $\text{SnBr}_4$ ,  $\text{SnI}_4$ ,  $\text{SnF}_2$ ,  $\text{SnCl}_2$ ,  $\text{SnBr}_2$  and  $\text{SnI}_2$ .

The gas to supply GSc may be diluted with an inert gas such as  $\text{H}_2$ ,  $\text{He}$ ,  $\text{Ar}$  and  $\text{Ne}$ , if necessary.

The lower layer may contain magnesium atoms (Mg). This is accomplished by introducing into the deposition chamber the raw materials to form the lower layer together with a raw material to introduce magnesium atoms (Mg) in a gaseous form. The raw material to supply magnesium atoms (Mg) may be gaseous at normal temperature and under normal pressure or gasifiable under the layer forming conditions.

The substance that can be used as a gas to supply magnesium atoms (Mg) include organometallic compounds containing magnesium atoms (Mg). Bis (cyclopentadienyl)-magnesium (II) complex salt ( $\text{Mg}(\text{C}_5\text{H}_5)_2$ ) is preferable from the standpoint of easy handling at the time of layer forming and the efficient supply of magnesium atoms (Mg).

The gas to supply magnesium atoms (Mg) may be diluted with an inert gas such as  $\text{H}_2$ ,  $\text{He}$ ,  $\text{Ar}$  and  $\text{Ne}$ , if necessary.

The lower layer may contain copper atoms (Cu). This is accomplished by introducing into the deposition chamber the raw materials to form the lower layer together with a raw material to introduce copper atoms (Cu) in a gaseous form. The raw material to supply copper atoms (Cu) may be gaseous at normal temperature and under normal pressure or gasifiable under the layer forming conditions.

The substance that can be used as a gas to supply copper atoms (Cu) include organometallic compounds containing copper atoms (Cu). Copper (II) bisdimethylglyoximate  $\text{Cu}(\text{C}_4\text{H}_7\text{N}_2\text{O}_2)_2$  is preferable from the standpoint of easy handling at the time of layer forming and the efficient supply of Cu atoms.

The gas to supply copper atoms (Cu) may be diluted with an inert gas such as  $\text{H}_2$ ,  $\text{He}$ ,  $\text{Ar}$  and  $\text{Ne}$ , if necessary.

The lower layer may contain sodium atoms (Na) or yttrium atoms (Y) or manganese atoms (Mn), zinc atoms (Zn), etc. This is accomplished by introducing into the deposition chamber the raw materials to form the lower layer together with a raw material to introduce sodium atoms (Na) or yttrium (Y) or manganese atoms (Mn) or zinc atoms (Zn). The raw material to supply sodium atoms (Na) or yttrium atoms (Y) or manganese atoms (Mn) or zinc atoms (Zn) may be gaseous at normal temperature and under normal pressure or gasifiable under the layer forming conditions.

18  
The substance that can be used as a gas to supply sodium atoms (Na) includes sodium amine ( $\text{NaNH}_2$ ) and organometallic compounds containing sodium atoms (Na). Among them, sodium amine ( $\text{NaNH}_2$ ) is preferable from the standpoint of easy handling at the time of layer forming and the efficient supply of sodium atoms (Na).

The substance that can be used as a gas to supply yttrium atoms (Y) includes organometallic compounds containing yttrium atoms (Y). Triisopropanol yttrium  $\text{Y}(\text{O}-\text{C}_3\text{H}_7)_3$  is preferable from the standpoint of easy handling at the time of layer forming and the efficient supply of yttrium atoms (Y).

The substance that can be used as a gas to supply manganese atoms (Mn) includes organometallic compounds containing manganese atoms (Mn). Monomethylpentacarbonyl-manganese  $\text{Mn}(\text{CH}_3)(\text{CO})_5$ , is preferable from the standpoint of easy handling at the time of layer forming and the efficient supply of sodium atoms (Na).

20 The substance that can be used as a gas to supply zinc atoms (Zn) includes organometallic compounds containing zinc atoms (Zn). Diethyl zinc  $\text{Zn}(\text{C}_2\text{H}_5)_2$  is preferable from the standpoint of easy handling at the time of layer forming and the efficient supply of zinc atoms (Zn).

25 The gas to supply sodium atoms (Na) or yttrium atoms (Y) or manganese atoms (Mn) or zinc atoms (Zn) may be diluted with an inert gas such as  $\text{H}_2$ ,  $\text{He}$ ,  $\text{Ar}$  and  $\text{Ne}$ , if necessary.

30 According to the present invention, the lower layer should have a thickness of  $0.03\text{--}5 \mu\text{m}$ , preferably  $0.01\text{--}1 \mu\text{m}$ , and most desirable  $0.05\text{--}0.5 \mu\text{m}$ , from the standpoint of the desired electrophotographic characteristics and economic effects.

35 According to the present invention, the lower layer has an interface region which is in contact with the aluminum support and contains less than 95% of the aluminum atoms contained in the aluminum support. If the interface region contains more than 95% of the 40 aluminum atoms contained in the aluminum support, it merely functions as the support. The lower layer also has an interface which is in contact with the upper layer and contains more than 5% of the aluminum atoms contained in the lower layer. If the interface region 45 contains less than 5% of the aluminum atoms contained in the lower layer, it merely functions as the upper layer.

In order to form the lower layer of  $\text{AlSiH}$  which has the characteristic properties to achieve the object of the present invention, it is necessary to properly establish the gas pressure in the deposition chamber and the temperature of the support.

The gas pressure in the deposition chamber should be properly selected according to the desired layer. It is usually  $1 \times 10^{-5}\text{--}10$  Torr, preferably  $1 \times 10^{-4}\text{--}3$  Torr, and most desirably  $1 \times 10^{-4}\text{--}1$  Torr.

The temperature ( $T_s$ ) of the support should be properly selected according to the desired layer. It is usually  $50^\circ\text{--}600^\circ \text{C}$ , and preferably  $100^\circ\text{--}400^\circ \text{C}$ .

In order to form the lower layer of  $\text{AlSiH}$  by the glow discharge method according to the present invention, it is necessary to properly establish the discharge electric power to be supplied to the deposition chamber according to the desired layer. It is usually  $5 \times 10^{-5}\text{--}10 \text{ W/cm}^3$ , preferably  $5 \times 10^{-4}\text{--}5 \text{ W/cm}^3$  and most desirably  $1 \times 10^{-3}\text{--}1$  to  $2 \times 10^{-3} \text{ W/cm}^3$ .

The gas pressure of the deposition chamber, the temperature of the support, and the discharge electric

power to be supplied to the deposition chamber mentioned above should be established interdependently to that the lower layer having the desired characteristic properties can be formed. Upper layer

The upper layer in this invention is composed of a 5 Non-Si (H, X) and has desired photoconductivity.

The upper layer of this invention contains, in at least the layer region adjacent with the lower layer, contained atoms (M) to control conductivity but contains no substantial carbon atoms (C), nitrogen atoms (N), oxygen atoms (O) germanium atoms (Ge) and tin atoms (Sn). However, the upper layer may contain in other layer regions at least one of the atoms (M) to control conductivity, carbon atoms (C), nitrogen atoms (N), oxygen atoms (O), germanium atoms (Ge) and tin atoms (Sn). Particularly, in the layer region of the upper layer near the free surface, at least one of carbon atoms (C), nitrogen atoms (N) and oxygen atoms (O) is preferably contained.

The upper layer may contain in the layer region of the upper layer at least adjacent with the lower layer optional atoms (M) to control conductivity, which are distributed evenly throughout the layer region or distributed evenly throughout the layer region but may be contained uneven distribution across the layer thickness in a part. However, in either of the cases, their distribution should be uniform in a plane parallel to the surface of the support so that uniform characteristics are ensured in the same plane.

In a case where the upper layer contains in other layer regions than the layer region at least in adjacent with the lower layer contains at least one of atoms (M) to control the conductivity, carbon atoms (C), nitrogen atoms (N), oxygen atoms (O), germanium atoms (Ge) and tin atoms (Sn), the atoms (M) to control the conductivity, carbon atoms (C), nitrogen atoms (N), oxygen atoms (O), germanium (Ge), tin atoms (Sn) may be distributed uniformly in the layer region, or they may be contained in a portion uniformly distributed in the layer region but not unevenly distributed across the layer thickness.

However, in either of the cases, their distribution should be uniform in a plane parallel to the surface of the support so that uniform characteristics are ensured in the same plane.

According to the present invention, the upper layer may contain at least one of alkali metals, alkaline earth metal and transition metals. The atoms are incorporated in the entire layer region or a partial layer region of the upper layer, and they may be uniformly distributed throughout the region, or distributed evenly through the layer region but may be contained unevenly distributed across the layer thickness.

However, they should be incorporated uniformly in either of the cases in a plane parallel to the surface of the support so that uniform characteristics are ensured in the same plane.

A layer region (hereinafter simply referred to as "layer region (CNO)") containing carbon atoms (C), and/or nitrogen atoms (N) and/or oxygen atoms (O) (hereinafter simply referred to as "atoms (CNO)"), a layer region (hereinafter simply referred to as "layer region (GS)") containing germanium atoms (Ge) and/or tin atoms (Sn) (hereinafter simply referred to as "atoms (GS)") and a layer region containing at least one alkali metals, alkaline earth metals and transition metals may have in common a layer region for a portion of the upper layer containing the layer region (M) to control

the conductivity (hereinafter simply referred to as "atoms (M)") on the surface of the layer region in adjacent at least with the lower layer (hereinafter simply referred to as "layer region (M<sub>B</sub>)").

Further, the layer region containing the atoms (M) other than the layer region (M<sub>B</sub>) (hereinafter simply referred to as "layer region (M<sub>T</sub>)") and the layer region (M<sub>B</sub>) and the layer region (M<sub>T</sub>) being collectively referred to as "layer region (M)", the layer region (CNO), the layer region (GS) and the layer region containing at least one of alkali metal atoms, alkaline earth metal atoms and transition metals may be a substantially identical layer region or may have in common a portion at least for each of the layer regions, or may not have in common a portion for each of the layer regions.

FIG. 17 to 36 show the typical examples of the profile of atoms (M) across the layer thickness in the layer region (M), a typical example of the profile of atoms (CNO) in the layer region (CNO) across the layer thickness, a typical example of the profile of the atoms (GS) contained the layer region (GS) across the layer thickness, and a typical example of the profile of alkali metal atoms, alkaline earth metal atoms or transition metal atoms contained in the layer region incorporating at least one of alkali metal atoms, alkaline earth metal atoms and transition metal atoms across the layer thickness in the upper layer of the light receiving member for use in electrophotography in this invention (hereinafter the layer regions are collectively referred to as "layer region (Y)" and these atoms are collectively referred to as "atoms (Y)").

Accordingly, FIG. 17 to 36 show the typical examples of the profiles of the atoms (Y) contained in the layer region (Y) across the layer thickness, in which one layer region (Y) is contained in the upper layer in a case where the layer region (M), layer region (CNO), layer region (GS), a layer region containing at least one of alkali metal, alkaline earth metal and transition metal are substantially the identical layer region, or a plurality of the layer regions (Y) are contained in the upper layer if they are not substantially identical layer region.

In FIGS. 17 to 36, the abscissa represents the distribution concentration C of the atoms (Y) and ordinate represents the thickness of the layer region (Y), while t<sub>B</sub> represents the position of the end of the layer region (Y) on the side of the layer and t<sub>T</sub> represents the position of the end of the layer region (Y) on the side of the free surface. That is, the layer region (Y) containing the atoms (Y) is formed from the side t<sub>B</sub> to the side t<sub>T</sub>.

FIG. 17 shows a first typical example of the profile of atoms (Y) contained in the layer region (Y) across the layer thickness.

In the example shown in FIG. 17, the atoms (Y) contained is distributed such that the concentration increases gradually and continuously from C<sub>171</sub> to C<sub>172</sub> from the position t<sub>B</sub> to the position t<sub>T</sub>.

In the example shown in FIG. 18, the atoms (Y) contained is distributed such that the concentration C linearly increases from C<sub>181</sub> to C<sub>182</sub> from the position t<sub>B</sub> to the position t<sub>181</sub> and takes a constant value of C<sub>183</sub> from the position t<sub>181</sub> to the position t<sub>T</sub>.

In the example shown in FIG. 19, the atoms (Y) contained is distributed such that the concentration C takes a constant value of C<sub>191</sub> from the position t<sub>B</sub> to the position t<sub>191</sub>, gradually and continuously increases from C<sub>191</sub> to C<sub>192</sub> from the position t<sub>191</sub> to the position t<sub>192</sub> and then takes a constant value of concentration t<sub>193</sub> from the position t<sub>192</sub> to the position t<sub>T</sub>.

In the example shown in FIG. 20, the atoms (Y) contained is distributed such that the concentration C takes a constant value of  $C_{201}$  from the position  $t_B$  to the position  $t_{201}$ , takes a constant value  $C_{202}$  from the position  $t_{201}$  to the position  $t_{202}$  and takes a constant value  $C_{203}$  from the position  $t_{202}$  to the position  $t_T$ .

In the example shown in FIG. 21, the atoms (Y) contained is distributed such that the concentration C takes a constant value of the  $C_{211}$  from the position  $t_B$  to the position  $t_T$ .

In the example shown in FIG. 22, the atoms (Y) contained is distributed such that the concentration C takes a constant value  $C_{221}$  from the position  $t_B$  to the position  $t_{221}$ , decreases gradually and continuously from  $C_{222}$  to  $C_{223}$  from the position  $t_{221}$  to the position  $t_T$ .

In the example shown in FIG. 23, the atoms (Y) contained is distributed such that the concentration C gradually and continuously decreases from  $C_{231}$  to the  $C_{232}$  from the position  $t_B$  to the position  $t_T$ .

In the example shown in FIG. 24 the atoms (Y) contained is distributed such that the distribution C takes a constant value  $C_{241}$  from the position  $t_B$  to the position  $t_{241}$ , gradually and continuously decreases from the  $C_{442}$  to the concentration substantially equal to zero from the position  $t_{241}$  to the position  $t_T$  (substantially zero means here and hereinafter the concentration lower than the detectable limit).

In the example shown in FIG. 25, the atoms (Y) contained is distributed such that the concentration C gradually and continuously decreases from  $C_{251}$  to substantially equal to zero from the position  $t_B$  to the position  $t_T$ .

In the example shown in FIG. 26, the atoms (Y) contained is distributed such that the concentration C remains constant at  $C_{261}$  from the position  $t_B$  to the position  $t_{262}$ , linearly decreases to  $C_{262}$  from the position  $t_{261}$  to the position  $t_T$  and remains at  $C_{262}$  at the position  $t_T$ .

In the example shown in FIG. 27, the atoms (Y) contained is distributed such that the concentration C linearly decreases from  $C_{271}$  to substantially equal to zero from the position  $t_B$  to the position  $t_T$ .

In the example shown in FIG. 28, the atoms (Y) contained is distributed such that the concentration C remaining constant at  $C_{281}$  from the position  $t_B$  to the position  $t_{281}$  and linearly decreases from  $C_{281}$  to  $C_{282}$  from the position  $t_{282}$  to the position  $t_T$ .

In the example shown in FIG. 29, the atoms (Y) contained is distributed such that the concentration C gradually and continuously decreases from  $C_{291}$  to  $C_{292}$  from the position  $t_B$  to the position  $t_T$ .

In the example shown in FIG. 30, the atoms (Y) contained is distributed such that the concentration C remains at a constant value  $C_{301}$  from the position  $t_B$  to the position  $t_{301}$ , linearly decreases from  $C_{302}$  to  $C_{303}$  from the position  $t_{301}$  to the position  $t_T$ .

In the example shown in FIG. 31, the atoms (Y) contained is distributed such that the concentration C gradually and continuously increases from  $C_{311}$  to  $C_{312}$  from the position  $t_B$  to the position  $t_{311}$  and remains at a constant value  $C_{313}$  from the position  $t_{311}$  to the position  $t_T$ .

In the example shown in FIG. 32, the atoms (Y) contained is distributed such that the concentration C gradually and continuously increases from  $C_{321}$  to  $C_{322}$  from the position  $t_B$  to the position  $t_T$ .

In the example shown in FIG. 33, the atoms (Y) contained is distributed such that the concentration C gradually and continuously increases from substantially zero to  $C_{331}$  from the position  $t_B$  to the position  $t_{331}$  and

remains constant at  $C_{332}$  between position  $t_{331}$  and position  $t_T$ .

In the example shown in FIG. 34, the atoms (Y) contained is distributed such that the concentration C gradually and continuously increases from substantially zero to  $C_{341}$  from the position  $t_B$  to the position  $t_T$ .

In the example shown in FIG. 35, the atoms (Y) contained is distributed such that the concentration C linearly increases from  $C_{351}$  to  $C_{352}$  from the position  $t_B$  to the position  $t_{351}$ , and remains constant at  $C_{352}$  from the position  $t_{351}$  to the position  $t_T$ .

In the example shown in FIG. 36, the atoms (Y) contained is distributed such that the concentration C linearly increases from  $C_{361}$  to  $C_{362}$  from the position  $t_B$  to the position  $t_T$ .

The atoms (M) to control the conductivity can include so-called impurities in the field of the semiconductor, and those used in this invention include atoms belonging to the group III of the periodical table giving p type conduction (hereinafter simply referred to as "group III atoms"), or atoms belonging to the group V of the periodical table except for nitrogen atoms (N) giving n-type conduction (hereinafter simply referred to as "group V atoms") and atoms belonging to the group VI of the periodical table except oxygen atoms (O) (hereinafter simply referred to as "group VI atoms").

Examples of the group III atoms can include B (boron), Al (aluminum), Ga (gallium), In (indium), Tl (thallium), etc., B, Al, Ga being particularly preferred. Examples of the group V atoms can include, specifically, P (phosphorus), As (arsenic), Sb (antimony), Bi (bismuth), P, As being particularly preferred. Examples of the group VI atoms can include, specifically, S (sulfur), Se (selenium), Te (tellurium) and Po (polonium), S and Se being particularly preferred. Incorporation of group III atoms, group V atoms or group VI atoms as the atoms (M) to control the conductivity into the layer region (M) in the present invention, can provide the effect, mainly, of controlling the conduction type and/or conductivity, and/or the effect of improving the charge injection between the layer region (M) and the lower region or selectively controlling for improving the charge inhibition, and/or the effect of improving the charge injection between the layer region (M) and the layer region other than the layer region (M) of the upper layer.

In the layer region (M), the content of atoms (M) to control the conductivity is preferably  $1 \times 10^{-3} - 5 \times 10^4$  atom-ppm, more preferably,  $1 \times 10^{-2} - 1 \times 10^4$  atom-ppm and, most preferably,  $1 \times 10^{-1} - 5 \times 10^3$  atom-ppm. Particularly, in a case where the layer region (M) contains carbon atoms (C), and/or nitrogen atoms (N), and/or oxygen atoms (O) described later by  $1 \times 10^3$  atom-ppm, the layer region (M) contains atoms (M) to control the conductivity preferably from  $1 \times 10^{-3} - 1 \times 10^3$  atom-ppm and, in a case if the content of the carbon atoms (C) and/or nitrogen atom (N) and/or oxygen atom (O) is in excess of  $1 \times 10^3$  atom-ppm, the content of the atoms (M) to control the conductivity is preferably  $1 \times 10^{-1} - 5 \times 10^4$  atom-ppm.

According to this invention, incorporation of the carbon atoms (C) and/or nitrogen atoms (N) and/or oxygen atoms (O) in the layer region (CNO) can mainly obtain an effect of increasing the dark resistance and/or hardness, and/or improving the control for the spectral sensitivity and/or enhancing the close bondability between the layer region (CNO) and the layer region of

the upper layer other than the layer region (CNO). The content of carbon atoms (C), and/or nitrogen atoms (N) and/or oxygen atoms (O) in the layer region (CNO) is preferably  $1-9\times 10^5$  atom-ppm, more preferably,  $1\times 10^1-5\times 10^5$  atom-ppm and most preferably,  $1\times 10^2-3\times 10^5$  atom-ppm. In addition, if it is intended to increase the dark resistance and/or the hardness, the content is preferably  $1\times 10^3-9\times 10^5$  atom-ppm and, preferably, it is  $1\times 10^2-5\times 10^5$  atom-ppm in a case where the spectral sensitivity is intended to be controlled.

In this invention, the spectral sensitivity can be controlled mainly and, particularly, sensitivity to the light of longer wave length can be improved in the case of using light of longer wavelength such as of a semiconductor laser for the image exposure source of electro-photographic apparatus by incorporating germanium atoms (Ge) and/or tin atoms (Sn) to the layer region (GS). The content of germanium atoms (Ge) and/or tin atoms (Sn) contained in the layer region is preferably  $1-9.5\times 10^5$  atom-ppm, more preferably,  $1\times 10^2-8\times 10^5$  atom-ppm and, most suitably,  $5\times 10^2-7\times 10^5$  atom-ppm.

In addition, hydrogen atoms (H) and/or halogen atoms (X) contained in the upper layer in this invention can compensate the unbonded bands of silicon atoms (Si), thereby improving the quality of the layer. The content of hydrogen atoms (H) or the sum of the hydrogen atoms (H) and halogen atoms (X) in the upper layer is suitably  $1\times 10^3-7\times 10^5$  atom-ppm, while the content of halogen atoms (X) is preferably  $1-4\times 10^5$  atom-ppm. Particularly, in a case where the content of the carbon atoms (C), and/or nitrogen atoms (N) and/or oxygen atoms (O) in the upper layer is less than  $3\times 10^5$  atom-ppm, the content of hydrogen atoms (H) or the sum of hydrogen atoms (H) and halogen atoms (X) is desirably  $1\times 10^3-4\times 10^5$  atom-ppm. Furthermore, in a case where the upper layer is composed of poly-Si(H,X), the content of hydrogen atoms (H) or the sum of hydrogen atoms (H) and halogen atoms (X) in the upper layer is preferably  $1\times 10^3-2\times 10^5$  atom-ppm and in a case where the upper layer is composed of A-Si(H,X), it is preferably  $1\times 10^4-7\times 10^5$  atom-ppm.

In this invention, the content of at least one of alkali metal, alkaline earth metal and transition metal in the upper layer is preferably  $1\times 10^{-3}-1\times 10^4$  atom-ppm, more preferably,  $1\times 10^{-2}-1\times 10^3$  atom-ppm and most suitably  $5\times 10^{-2}-5\times 10^2$  atom-ppm.

In this invention, the upper layer composed of Non-Si(H,X) can be prepared by the same vacuum deposition film formation as that for the lower layer described above, and glow discharge, sputtering, ion plating, HRCVD process, FOCVD process are particularly preferred. These methods may be used in combination in one identical device system.

For instance, the glow discharge method may be performed in the following manner to form the upper layer composed of Non-Si(H,X). The raw material gases are introduced into an evacuable deposition chamber and glow discharge is performed with the gases being introduced at a desired pressure, so that a layer of Non-Si(H,X) is formed as required on the surface of the support situated at a predetermined position and previously formed with a predetermined lower layer. The raw material gases may contain a gas to supply silicon atoms (Si), a gas to supply hydrogen atoms (H), and/or a gas to supply halogen atoms (X), an optional gas to supply atoms (M) to control the conduc-

tivity, and/or a gas to supply carbon atoms (C), and/or a gas to supply nitrogen atoms (N), and/or a gas to supply oxygen atoms (O), and/or a gas to supply germanium atoms (Ge), and/or a gas to supply tin atoms (Sn) and/or a gas to supply at least one of alkali metal, alkaline earth metal and transition metal.

The HRCVD process may be performed in the following manner to form the upper layer composed of Non-Si(H,X). The raw material gases are introduced individually or altogether into an evacuable deposition chamber, and glow discharge performed or the gases are heated with the gases being introduced at a desired pressure, during which active substance (A) is formed and another active substance (B) is introduced into the deposition chamber, so that a layer of Non-Si(H,X) is formed as required on the surface of the support situated at a predetermined position and formed with a predetermined lower layer thereon in the deposition chamber. The raw material gases may contain a gas to supply silicon atoms (Si), a gas to supply halogen atoms (X), an optional gas to control conductivity (M), and/or a gas to supply carbon atoms (C), and/or a gas to supply nitrogen atoms (N), and/or a gas to supply oxygen atoms (O), and/or a gas to supply germanium atoms (Ge), and/or a gas to supply tin atoms (Sn) and/or a gas to supply at least one of alkali metal, alkaline earth metal and transition metal. Another active substance (B) is formed by introducing a gas to supply hydrogen activation space. The active substance (A) and another active substance (B) may individually be introduced into the deposition chamber.

The FOCVD process may be performed in the following manner to form the upper layer of Non-Si(H,X). The raw material gases are introduced into an evacuable deposition chamber individually or altogether as required under a desired gas pressure. The raw material gases may contain a gas to supply silicon atoms (Si), a gas to supply hydrogen atoms (H), an optional gas to supply atoms (M) to control conductivity, and/or a gas to supply carbon atoms (C), and/or a gas to supply nitrogen atoms (N), and/or a gas to supply oxygen atoms (O), and/or a gas to supply germanium atoms (Ge), and/or a gas to supply tin atoms (Sn) and/or a gas to supply at least one of alkali metal, alkaline earth metal and transition metals. They may be introduced into the deposition chamber individually or altogether as required. A halogen (X) gas is introduced into the deposition chamber separately from the raw material gases described above and these gases subjected to chemical reactions in the deposition chamber.

The sputtering method or the ion plating method may be performed in the following manner to form the upper layer composed of the Non-Si(H,X), basically, by the known method as described for example, in Japanese Patent Laid-Open No. Sho 61-59342.

According to this invention, the upper layer is formed while controlling the profile of the concentration C of atoms (M) to control the conductivity, carbon atoms (C), nitrogen atoms (N), oxygen atoms (O), germanium atoms (Ge), tin atoms (Sn) and at least one of alkali metal atoms, alkaline earth metal atoms and transition metal atoms (simply referred to collectively as "atoms (Z)") across the layer thickness to obtain a layer having a desired depth profile across the layer thickness. This can be achieved, in the case of glow discharge, HRCVD and FOCVD, by properly controlling the gas flow rate of a gas to supply atoms (Z) the concentration of which is to be varied in accordance with a

desired rate of change in the concentration and then introducing the gas into the deposition chamber.

The flow rate may be changed by operating a needle valve disposed in the gas passage manually or by means of a customary means such as an external driving motor.

Alternatively, the flow rate setting to a mass flow controller for the control of the gas flow rate is properly changed by an adequate means manually or using a programmable control device.

The gas to supply Si atoms used in this invention can include gaseous or gasifiable silicon hydrides (silanes) such as SiH<sub>4</sub>, Si<sub>2</sub>H<sub>6</sub>, Si<sub>3</sub>H<sub>8</sub> and Si<sub>4</sub>H<sub>10</sub>. SiH<sub>4</sub> and Si<sub>2</sub>H<sub>6</sub> are preferable from the standpoint of ease of handling and the efficient supply of Si. These gases to supply Si may be diluted with an inert gas such as H<sub>2</sub>, He, Ar and Ne if necessary.

According to the present invention, the gas to supply halogen includes various halogen compounds, for example, gaseous and gasifiable halogen compounds, for example, halogen gases, halides, interhalogen compounds and halogen-substituted silane derivatives.

Additional examples in this invention can include, gaseous or gasifiable halogen atom (X)-containing silicon hydride compounds composed of silicon atoms (Si) and halogen atoms (X).

Halogen compounds that can be suitably used in this invention can include halogen gases such as of fluorine, chlorine, bromine and iodine; and interhalogen compounds such as BrF, ClF, ClF<sub>3</sub>, BrF<sub>5</sub>, BrF<sub>3</sub>, IF<sub>3</sub>, IF<sub>7</sub> ICl and IBr.

Examples of the halogen atoms (X)-containing silicon compounds, or halogen atom (X)-substituted silane derivatives can include, specifically, silicon halides such as SiF<sub>4</sub>, Si<sub>2</sub>F<sub>6</sub>, SiCl<sub>4</sub> and SiBr<sub>4</sub>.

In the case where the halogen-containing silicon compound is used to form the light receiving member for use in electrophotography according to this invention by the glow discharge or HRCVD method, it is possible to form the upper layer composed of Non-Si(H,X) containing halogen atoms (X) on a desired lower layer without using a silicohydride gas to supply Si atoms.

In the case where the upper layer containing halogen atoms (X) is formed according to the glow discharge or HRCVD method, a silicon halide gas is used as the gas to supply silicon atoms to form the upper layer on a desired support. The silicon halide gas may further be mixed with hydrogen gas or a hydrogen atom (H)-containing silicon compound gas to facilitate the introduction of hydrogen atoms (H) at a desired level.

The above-mentioned gases may be used individually or in combination with one another at a desired mixing ratio.

In this invention, the above-mentioned halogen compounds or halogen atom (X)-containing silicon compounds are used as effective material as the gas to supply halogen atoms, but gaseous or gasifiable hydrogen halides such as HF, HCl, HBr and HI; and halogen-substituted silicohydrides such as SiH<sub>3</sub>F, SiH<sub>2</sub>F<sub>2</sub>, SiHF<sub>3</sub>, SiH<sub>2</sub>I<sub>1</sub>, SiH<sub>2</sub>Cl<sub>2</sub>, SiHCl<sub>3</sub>, SiH<sub>2</sub>Br<sub>2</sub> and SiBr<sub>3</sub> can also be used. Among them, hydrogen atom (H)-containing halides can be used as preferably halogen supply gases in this invention upon forming the upper layer, because they supply the upper layer with halogen atoms (X), as well as hydrogen atoms (H) which are very effective for the control of electric or photoelectric characteristics.

The introduction of hydrogen atoms (H) into the upper layer may also be accomplished in another

method by inducing discharge in the deposition chamber containing H<sub>2</sub> or silicohydride such as SiH<sub>4</sub>, Si<sub>2</sub>H<sub>6</sub>, Si<sub>3</sub>H<sub>8</sub> and Si<sub>4</sub>H<sub>10</sub> and a silicon compound to supply silicon atoms (Si).

5 The amount of hydrogen atoms (H) and/or halogen atoms (X) to be introduced into the upper layer may be controlled by regulating the temperature of the support, the amount of raw materials for hydrogen atoms and halogen atoms to be introduced into the deposition chamber and/or the electric power for discharge.

The upper layer may contain atoms (M) to control the conductivity, for example, group III atoms, group V atoms or group VI atoms. This is accomplished by introducing into the deposition chamber the raw materials to form the upper layer together with a raw materials to supply group III atoms, raw materials to supply group V atoms or raw material to supply group VI atoms. The raw material to supply group III atoms, the raw material to supply group V atoms, or the raw material to supply group VI atoms may be gaseous at normal temperature and under normal pressure or gasifiable under the layer forming conditions are desirably used. The raw material to supply the group III atoms can include specifically boron hydrides such as B<sub>2</sub>H<sub>6</sub>, B<sub>4</sub>H<sub>10</sub>, B<sub>4</sub>H<sub>9</sub>, B<sub>5</sub>H<sub>11</sub>, B<sub>6</sub>H<sub>10</sub>, B<sub>6</sub>H<sub>12</sub> and B<sub>6</sub>H<sub>14</sub> or boron hydrides such as BF<sub>3</sub>, BCl<sub>3</sub> and BBr<sub>3</sub> for the material to supply boron atoms. Additional examples are AlCl<sub>3</sub>, GaCl<sub>3</sub>, Ga(CH<sub>3</sub>)<sub>3</sub>, InCl<sub>3</sub> and TiCl<sub>3</sub>.

20 The raw material to supply group V atoms that can be used effectively in this present invention can include, phosphorus hydride such as PH<sub>3</sub>, P<sub>2</sub>H<sub>4</sub>, etc. phosphorus halide such as PH<sub>4</sub>I, PF<sub>3</sub>, PF<sub>5</sub>, PCl<sub>3</sub>, PCl<sub>5</sub>, PBr<sub>3</sub>, PBr<sub>5</sub> and PI<sub>3</sub> as the material to supply phosphorus atoms.

25 Additional examples as effective raw materials to supply group V atoms can also include AsH<sub>3</sub>, AsF<sub>3</sub>, AsCl<sub>3</sub>, AsBr<sub>3</sub>, AsF<sub>5</sub>, SbH<sub>3</sub>, SbF<sub>3</sub>, SbF<sub>5</sub>, SbCl<sub>3</sub>, SbCl<sub>5</sub>, BiH<sub>3</sub>, BiCl<sub>3</sub>, BiBr<sub>3</sub>.

30 Raw materials to supply groups VI atoms can include those gaseous or gasifiable materials such as hydrogen sulfide (H<sub>2</sub>S), SF<sub>4</sub>, SV<sub>6</sub>, SO<sub>2</sub>, SO<sub>2</sub>F<sub>2</sub>, COS, CS<sub>2</sub>, CH<sub>3</sub>SH, C<sub>2</sub>H<sub>5</sub>SH, C<sub>4</sub>H<sub>4</sub>S, (CH<sub>3</sub>)<sub>2</sub>S, (C<sub>2</sub>H<sub>5</sub>)<sub>2</sub>S, etc. Additional example can include, those gaseous or gasifiable materials such as SeH<sub>2</sub>, SeF<sub>6</sub>, (CH<sub>3</sub>)<sub>2</sub>Se, (C<sub>2</sub>H<sub>5</sub>)<sub>2</sub>Se, TeH<sub>2</sub>, TeF<sub>6</sub>, (CH<sub>3</sub>)<sub>2</sub>Te, (C<sub>2</sub>H<sub>5</sub>)<sub>2</sub>Te.

35 The raw material for supplying atoms (M) to control the conductivity may be diluted with an inert gas such as H<sub>2</sub>, He, Ar and Ne if necessary.

40 The upper layer may contain carbon atoms (C), nitrogen atoms (N) or oxygen atoms (O). This accomplished by introducing into the chamber the raw material to supply carbon atoms (C), the raw material to supply nitrogen atoms (N) or raw material to supply oxygen atoms (O) in a gaseous form together with other raw materials for forming the upper layer. The raw material to supply carbon atoms (C), the raw material to supply nitrogen atoms (N) or the raw material to supply oxygen atoms (O) are desirably gaseous at normal temperature and under normal pressure or gasifiable under the layer forming conditions.

45 A raw material that can effectively be used as the starting gas to supply carbon atoms (C) can include those hydrocarbons having C and H as constituent atoms, for example, saturated hydrocarbons having 1 to 4 carbon atoms, ethylene series hydrocarbons having 2 to 4 carbon atoms and acetylene series hydrocarbon atoms 2 to 3 carbon atoms.

50 Examples of the saturated hydrocarbons include methane (CH<sub>4</sub>), ethane (C<sub>2</sub>H<sub>6</sub>), propane (C<sub>3</sub>H<sub>8</sub>), n-

butane (n-C<sub>4</sub>H<sub>10</sub>), pentane (C<sub>5</sub>H<sub>12</sub>). Examples of ethylene series hydrocarbons include ethylene (C<sub>2</sub>H<sub>4</sub>), propylene (C<sub>3</sub>H<sub>6</sub>), butene-1 (C<sub>4</sub>H<sub>8</sub>), butene-2 (C<sub>4</sub>H<sub>8</sub>), isobutylene (C<sub>4</sub>H<sub>8</sub>) and pentene (C<sub>5</sub>H<sub>10</sub>). Examples of acetylene series hydrocarbon can include, acetylene (C<sub>2</sub>H<sub>2</sub>), methylacetylene (C<sub>3</sub>H<sub>4</sub>) and butine (C<sub>4</sub>H<sub>6</sub>).

Additional example can include halogenated hydrocarbon gases such as CF<sub>4</sub>, CCl<sub>4</sub> and CH<sub>3</sub>CF<sub>3</sub> with a view point that halogen atom (X) can be introduced in addition to hydrocarbons (C).

Examples of the raw materials gas to introduce nitrogen atoms (N) can include those having N as constituent atoms, or N and H as constituent atoms, for example, gaseous or gasifiable nitrogen, or nitrogen compounds such as nitrides and azides, for example, nitrogen (N<sub>2</sub>), ammonia (NH<sub>3</sub>), hydrazine (H<sub>2</sub>NNH<sub>2</sub>), hydrogen azide (HN<sub>3</sub>) and ammonium azide (NH<sub>4</sub>N<sub>3</sub>). Additional examples can include halogenated nitrogen compounds such as nitrogen trifluoride (F<sub>3</sub>N) and nitrogen tetrafluoride (F<sub>4</sub>N<sub>2</sub>), etc. which can introduce nitrogen atoms as well as halogen atoms (X).

Examples of the raw material gas to introduce oxygen atoms (O) can include oxygen (O<sub>2</sub>), ozone (O<sub>3</sub>), nitrogen monoxide (NO), nitrogen dioxide (NO<sub>2</sub>), dinitrogen oxide (N<sub>2</sub>O), dinitrogen trioxide (N<sub>2</sub>O<sub>3</sub>), trinitrogen tetraoxide (N<sub>3</sub>O<sub>4</sub>), dinitrogen pentaoxide (N<sub>2</sub>O<sub>5</sub>) and nitrogen trioxide (NO<sub>3</sub>), as well as lower siloxanes having silicon atoms (Si), oxygen atoms (O) and hydrogen atoms (H) as constituent atoms, for example, disiloxane (H<sub>3</sub>SiOSiH<sub>3</sub>) and trisiloxane (H<sub>3</sub>SiOSiH<sub>2</sub>OSiH<sub>3</sub>).

The upper layer may be introduced with germanium (Ge) or tin atoms (Sn). This is accomplished by introducing, into the deposition chamber, the raw material to supply germanium (Ge) or the raw material to supply tin atoms (Sn) into the deposition chamber together with other raw materials to form the upper layer in a gaseous form. The raw material to supply germanium (Ge) or the raw material to supply tin atoms (Sn) may desirably be gaseous at normal temperature and normal pressure or gasifiable under the layer forming conditions.

The material that can be used as a gas to supply germanium atoms (Ge) can include, gaseous or gasifiable germanium hydrides such as GeH<sub>4</sub>, Ge<sub>2</sub>H<sub>6</sub>, Ge<sub>3</sub>H<sub>8</sub> and Ge<sub>4</sub>H<sub>10</sub>, and GeH<sub>4</sub>, Ge<sub>2</sub>H<sub>6</sub> and Ge<sub>3</sub>H<sub>8</sub> being preferable from the standpoint of easy handling at the time of layer forming and the efficient supply of germanium atoms (Ge).

Additional examples of the raw material for effectively forming the upper layer can include those gaseous or gasifiable materials such as germanium hydride-halides, for example, GeHF<sub>3</sub>, GeH<sub>2</sub>F<sub>2</sub>, GeH<sub>3</sub>F, GeHCl<sub>3</sub>, GeH<sub>2</sub>Cl<sub>2</sub>, GeH<sub>3</sub>Cl, GeHBr<sub>3</sub>, GeH<sub>2</sub>Br<sub>2</sub>, GeH<sub>3</sub>Br, GeHI<sub>3</sub>, GeH<sub>2</sub>I<sub>2</sub> and GeH<sub>3</sub>I, as well as germanium halides such as GeF<sub>4</sub>, GeCl<sub>4</sub>, GeBr<sub>4</sub>, GeI<sub>4</sub>, GeF<sub>2</sub>, GeCl<sub>2</sub>, GeBr<sub>2</sub> and GeI<sub>2</sub>.

The material that can be used as a gas to supply tin atoms (Sn) can include gaseous or gasifiable tin hydrides such as SnH<sub>4</sub>, Sn<sub>2</sub>H<sub>6</sub>, Sn<sub>3</sub>H<sub>8</sub> and Sn<sub>4</sub>H<sub>10</sub> and SnH<sub>4</sub>, Sn<sub>2</sub>H<sub>6</sub> and Sn<sub>3</sub>H<sub>8</sub> being preferred from the standpoint of easy handling at the time of layer forming and the efficient supply of tin atoms (Sn).

Additional examples of the starting material for effectively forming the upper layer can include gaseous or gasifiable tin halide-hydrides such as SnHF<sub>3</sub>, SnH<sub>2</sub>F<sub>2</sub>, SnH<sub>3</sub>F, SnHCl<sub>3</sub>, SnH<sub>2</sub>Cl<sub>2</sub>, SnH<sub>3</sub>Cl, SnHBr<sub>3</sub>, SnH<sub>2</sub>Br<sub>2</sub>, SnH<sub>3</sub>Br, SnHI<sub>3</sub>, SnH<sub>2</sub>I<sub>2</sub> and SnH<sub>3</sub>I, as well as tin ha-

lides such as SnF<sub>4</sub>, SnCl<sub>4</sub>, SnBr<sub>4</sub>, SnI<sub>4</sub>, SnF<sub>2</sub>, SnCl<sub>2</sub>, SnBr<sub>2</sub> and SnI<sub>2</sub>.

The lower layer may contain magnesium atoms (Mg). This is accomplished by introducing, into the deposition chamber, the raw materials for supplying magnesium atoms (Mg) to form the upper layer together with other raw materials for forming the upper layer in a gaseous form. The raw material to supply magnesium atoms (Mg) may be gaseous at normal temperature and a normal pressure or gasifiable under the layer forming conditions.

The substance that can be used as a gas to supply magnesium atoms (Mg) can include organometallic compounds containing magnesium atoms (Mg). Bis(cyclopentadienyl)-magnesium (II) complex salt (Mg(C<sub>5</sub>H<sub>5</sub>)<sub>2</sub>) is preferable from the stand point of easy handling at the time of layer form an the effective supply of magnesium atoms (Mg).

The gas to supply magnesium atoms (Mg) may be diluted with an inert gas such as H<sub>2</sub>, He, Ar and Ne if necessary.

The upper layer may contain copper atoms (Cu). This is accomplished by introducing, into the deposition chamber, the raw material to supply copper atoms (Cu) for forming the upper layer together with other raw materials for forming the upper layer in a gaseous form. The raw material to supply copper atoms (Cu) may be gaseous at normal temperature and normal pressure and gasifiable under the layer forming condition.

The material that can be used as a gas to supply copper atoms (Cu) can include organometallic compounds containing copper atoms (Cu). Copper (II)bisdimethylglyoximate CU(C<sub>4</sub>N<sub>2</sub>O<sub>2</sub>)<sub>2</sub> is preferred from the stand point of easy handling at the time of layer forming and efficient supply of magnesium atoms (Mg).

The gas to supply copper atoms (Cu) may be diluted with an inert gas such as H<sub>2</sub>, He, Ar and Ne, if necessary.

The upper layer may contain sodium atoms (Na), yttrium atoms (Y), manganese atoms (Mn) or zinc atoms (Zn). This is accomplished by introducing, into the deposition chamber, raw material to supply sodium atoms (Na), the raw material to supply yttrium atoms (Y), the raw material to supply manganese atoms (Mn) or the raw materials to supply zinc atoms (Zn) for forming the upper layer together with other raw materials for forming the upper layer in a gaseous form. The raw material to supply sodium atoms (Na), the raw material to supply yttrium atoms (Y), the raw material to supply manganese atoms (Mn) or the raw material to supply zinc atoms (Zn) may be gaseous at normal temperature and normal pressure or gasifiable at least under the layer forming conditions.

The material that can be effectively used as a gas to supply sodium atoms (Na) can include sodium amine (NaNH<sub>2</sub>) and organometallic compounds containing sodium atoms (Na). Among them, sodium amine (NaNH<sub>2</sub>) is preferred from the standpoint of easy handling at the time of layer forming and the efficient supply of sodium atoms (Na).

The material that can be effectively used as a gas to supply yttrium atoms (Y) can include organometallic compounds containing yttrium atoms (Y). Triisopropanol yttrium Y(Oi-C<sub>3</sub>H<sub>7</sub>)<sub>3</sub> is preferred from the standpoint of easy handling at the time of layer forming and the effective supply of yttrium atoms (Y).

The material can be effectively used as a gas to supply manganese atoms (Mn) can include organometallic

compounds containing manganese atoms (Mn). Monomethylpentacarbonyl manganese  $Mn(CH_3)(CO)_5$  is preferred from the standpoint of easy handling at the time of layer forming and the efficient supply of manganese atoms (Mn).

The material that can be effectively used as a gas to supply zinc atoms (Zn) can include organometallic compounds containing Zinc atoms (Zn). Diethyl zinc  $Zn(C_2H_5)_2$  is preferred from the standpoint of easy handling at the time of layer forming and the efficient supply of zinc atoms (Zn).

The gas to supply sodium atoms (Na), yttrium atoms (Y), manganese atoms (Mn) or zinc atoms (Zn) may be diluted with an inert gas such as  $H_2$ , He, Ar and Ne, if necessary.

In the present invention, the layer thickness of the upper layer is 1-130  $\mu m$ , preferably, 3-100  $\mu m$  and, most suitably, 5-60  $\mu m$  from the standpoint of the desired electrophotographic characteristics and economical effect.

In order to form the upper layer composed of Non-Si(H,X) which has the characteristics to achieve the object of this invention, it is necessary to properly establish the gas pressure in the deposition chamber and the temperature of the support.

The gas pressure in the deposition chamber should properly be selected according to the design of the layer. It is usually  $1 \times 10^{-5}$  - 10 Torr, preferably,  $1 \times 10^{-4}$  - 3 Torr and, most suitably,  $1 \times 10^{-4}$  - 1 Torr. In the case of selecting A-Si(H, X) as the Non-Si(H,X) for the upper layer, the temperature (Ts) of the support should properly be selected according to the desired design for the layer and it is usually 50°-400° C., preferably, 100°-300° C. In a case where poly-Si(H,X) is selected as the Non-Si(H,X) for the upper layer, there are various methods for forming the layer including, for example, the following methods.

In one method, the temperature of the support is set to a high temperature, specifically, to 400°-600° C. and a film is deposited on the support by means of the plasma CVD process.

In another method, an amorphous layer is formed at first to the surface of the support. That is, a film is formed on a support heated to a temperature of about 250° C. by a plasma CVD process and the amorphous layer is annealed into a polycrystalline layer. The annealing is conducted by heating the support to 400°-600° C. about for 5-30 min, or applying laser beams for about 5-30 min.

Upon forming the upper layer composed of Non-Si(H,X) by the glow discharge method according to this invention, it is necessary to properly select the discharge electric power to be supplied to the deposition chamber according to the design of the layer. It is usually  $5 \times 10^{-5}$  - 10 W/cm<sup>3</sup>, preferably,  $5 \times 10^{-5}$  - 5 W/cm<sup>3</sup> and, most suitably,  $1 \times 10^{-3}$  -  $2 \times 10^{-1}$  W/cm<sup>3</sup>.

The gas pressure of the deposition chamber, the temperature of the support and the discharge electric power to be supplied to the deposition chamber mentioned above should be set interdependently so that the upper layer having the desired characteristic properties can be formed.

#### EFFECT OF THE INVENTION

The light receiving member for use in electrophotography according to this invention, having the specific layer structure as described above, can overcome all of the problems in the conventional light receiving mem-

bers for use in electrophotography constituted with A-Si and it can exhibit particularly excellent electrical properties, optical properties, photoconductive properties, image properties, durability and characteristics in the circumstance of use.

Particularly, since the lower layer contains aluminum atoms (Al), silicon atoms (Si) and, particularly, hydrogen atoms (H) across the layer thickness in an unevenly distributed state according to the present invention, injection of charges (photocarriers) across the aluminum support and the upper layer can be improved and, moreover, since the texture and continuity for the constituent elements between the aluminum support and the upper layer is improved, image properties such as coarse image or dots can be improved thereby enabling to stably reproduce high quality images with clear half-tone and high resolving power.

In addition, it is possible to prevent image defects or peeling of Non-Si(H,X) films due to impactive mechanical pressure applied for a relatively short period of time to the light receiving member for use in electrophotography, thereby improving the durability and, further, stresses resulted from the difference in the heat expansion coefficients between aluminum support and Non-Si(H,X) film to prevent cracking or peeling in the Non-Si(H,X) film to thereby enhance the yield of the productivity.

Incorporation of at least one of atoms, to control conductivity into the layer region of the upper layer in 30 adjacent with the lower layer can improve the charge injection or selectively controlling or improving the charge inhibition between the upper layer and the lower layer, to prevent the occurrence of image defects such as coarse image or dots, as well as high quality image with clear half-tone and high resolving power can be reproduced stably and durability teh charging power and the can also be improved. durability.

Further, since atoms (Mc) to control the image quality are contained in the lower layer in addition to aluminum atoms (Al), silicon atoms (Si) and hydrogen atoms (H), the injection of photocarriers across the aluminum support and the upper layer is further improved and the transferability of the photocarriers in the lower layer is improved. Accordingly, image characteristics such as coarse image can be improved to stably reproduce a high quality image with clear half-tone and high resolving power.

Furthermore, since halogen atoms co-existent in the lower layer can compensate dangling bonds of silicon atoms aluminum atoms, etc. to attain more stable state in view of the texture and structure according to the present invention, remarkable improvement can be obtained in view of the image characteristics such as coarse image or dots coupled with the foregoing effect due to the distribution of the silicon atoms, aluminum atoms and hydrogen atoms.

Since at least one of germanium atoms (Ge) and tin atoms (Sn) are contained in the lower layer according to this invention, the injection of the photocarriers across the aluminum support and the upper layer, close bondability and the transferability of the photocarriers in the lower layer can remarkably be improved to thereby provide remarkable improvement in the characteristics and durability of a light receiving member.

Particularly, since at least one of alkali metal atoms, alkaline earth metal atoms and transition metal atoms are contained in the upper layer according to the present invention, an outstanding feature can be obtained

that the hydrogen atoms and halogen atoms contained in the lower layer can be dispersed more effectively to prevent layer peeling resulted from the cohesion of hydrogen atoms and/or halogen atoms during long time use.

Furthermore, since the injection of photocarriers and the close bondability across the aluminum support and the upper layer, and the transferability of photocarriers in the lower layer can be improved remarkably as described above, significant improvement can be obtained in the image property and the durability to result in improvement to stable production of the lightreceiving member having a stable quality.

#### PREFERRED EMBODIMENT OF THE INVENTION

This invention will be described more specifically referring to examples but the invention is no way limited only thereto.

#### EXAMPLE 1

A light receiving member for use in electrophotography according to this invention was formed by radio frequency (hereinafter simply referred to as "RF") glow discharge decomposition.

FIG. 37 shows an apparatus for producing the light receiving member for use in electrophotography by the RF glow discharge decomposition, comprising a raw material gas supply device 1020 and a deposition device 1000.

In the figure, raw material gases for forming the respective layers in this invention were tightly sealed in gas cylinders 1071, 1072, 1073, 1074, 1075, 1076 and 1077, and a tightly sealed vessel 1078, in which the cylinder 1071 was for SiH<sub>4</sub> gas (99.99% purity), the cylinder 1072 was for H<sub>2</sub> gas (99.9999%), the cylinder 1073 was for CH<sub>4</sub> gas (99.999% purity), cylinder 1074 was for PH<sub>3</sub> gas diluted with H<sub>2</sub> gas (99.999% purity, hereinafter simply referred to as "PH<sub>3</sub>/H<sub>2</sub>"), the cylinder 1075 was for B<sub>2</sub>H<sub>6</sub> gas diluted with H<sub>2</sub> gas (99.999% purity, hereinafter simply referred to as "B<sub>2</sub>H<sub>6</sub>/H<sub>2</sub>"), the cylinder 1076 was for N<sub>2</sub> gas (99.9999% purity), the cylinder 1077 was for He gas (99.999% purity), and the tightly sealed vessel 1078 was for AlCl<sub>3</sub> (99.99% purity).

In the figure, a cylindrical aluminum support 1005 had an outer diameter of 108 mm and a mirror-finished surface.

After confirming that valves 1051-1057 for the gas cylinders 1071-1077, flow-in valves 1031-1037 and a leak valve 1015 for the deposition chamber 1001 were closed and flow-out valves 1041-1047 and an auxiliary valve 1018 were opened, a main valve 1016 was at first opened to evacuate the deposition chamber 1001 and gas pipeways by a vacuum pump not illustrated.

Then, when the indication of a vacuum meter 1017 showed about  $1 \times 10^{-3}$  Torr, the auxiliary valve 1018, the flow-out valves 1041-1047 were closed.

Then, the valves 1051-1057 were opened to introduce SiH<sub>4</sub> from the gas cylinder 1071, H<sub>2</sub> gas from the gas cylinder 1072, CH<sub>4</sub> gas from the gas cylinder 1073, PH<sub>3</sub>/H<sub>2</sub> gas from the gas cylinder 1074, B<sub>2</sub>H<sub>6</sub>/H<sub>2</sub> gas from the gas cylinder 1075, N<sub>2</sub> gas from the gas cylinder 1076 and He gas from the gas cylinder 1077, and the pressures for the respective gases were adjusted to 2 kg/cm<sup>2</sup> by pressure controllers 1061-1067.

Then, the flow-in valves 1031-1037 were gradually opened to introduce the respective gases in mass flow

controllers 1021-1027. In this case, since the He gas from the gas cylinder 1077 was passed through the tightly sealed vessel 1078 charged with AlCl<sub>3</sub>, the AlCl<sub>3</sub> gas diluted with the He gas (hereinafter simply referred to as "AlCl<sub>3</sub>/He") was introduced to the mass flow controller 1027.

The temperature of the cylindrical aluminum support 1005 disposed in the deposition chamber 1001 was heated to 250° C. by a heater 1014.

After completing the preparation for the film formation as described above, each of the lower and upper layers was formed on the cylindrical aluminum support 1005.

The lower layer was formed by gradually opening the flow-out valves 1041, 1042 and 1047, and the auxiliary valve 1018 thereby introducing the SiH<sub>4</sub> gas, H<sub>2</sub> gas and AlCl<sub>3</sub>/He gas through the gas discharge aperture 1009 of a gas introduction pipe 1018 to the inside of the deposition chamber 1001. In this case, the gas flow rates were controlled by the respective mass flow controllers 1021, 1022 and 1027 such that the gas flow rates were set to 50 SCCM for SiH<sub>4</sub>, 10 SCCM for H<sub>2</sub> gas, and 120 SCCM for AlCl<sub>3</sub>/He. The pressure in the deposition chamber was controlled to 0.4 Torr by adjusting the opening of the main valve 1016 while observing the vacuum meter 1017. Then, RF power was introduced to the inside of the deposition chamber 1001 by way of an RF matching box 1012 while setting the power of a RF power source (not illustrated) to 5 mW/cm<sup>3</sup>, to cause RF glow discharge, thereby starting the formation of the lower layer on the aluminum support. The mass flow controllers 1021, 1022 and 1027 were adjusted during formation of the lower layer such that the SiH<sub>4</sub> gas flow remains at a constant rate of 50 SCCM, the H<sub>2</sub> gas flow rate is increased at a constant ratio from 10 SCCM to 200 SCCM and the AlCl<sub>3</sub>/He gas flow rate is decreased at a constant ratio from 120 SCCM to 40 SCCM. Then, when the lower layer of 0.05 μm thickness was formed, the RF glow discharge was stopped and the entrance of the gas to the inside of the deposition chamber 1001 is interrupted by closing the flow-out valves 1041, 1042 and 1047 and the auxiliary valve 1018, to complete the formation of the lower layer.

Then, for forming the first layer region of the upper layer, the flow-out valves 1041, 1042 and 1045, and the auxiliary valve 1018 were gradually opened to flow SiH<sub>4</sub> gas, H<sub>2</sub> gas and B<sub>2</sub>H<sub>6</sub>/H<sub>2</sub> gas through the gas discharge aperture 1009 of the gas introduction pipe 1008 into the deposition chamber 1001. In this case, respective mass flow controllers 1021, 1022 and 1025 were adjusted so that the SiH<sub>4</sub> gas flow rate was 100 SCCM, H<sub>2</sub> gas flow rate was 500 SCCM and B<sub>2</sub>H<sub>6</sub>/H<sub>2</sub> gas flow rate was 200 ppm to SiH<sub>4</sub>. The pressure in the deposition chamber 1001 was controlled to 0.4 Torr by adjusting the opening of the main valve 1016 while observing the vacuum meter 1017. Then, RF power was introduced into the deposition chamber 1001 through a radio frequency matching box 1012 while setting the power of a RF power source (not illustrated) to 8 mW/cm<sup>3</sup>, to cause RF glow discharge and start the formation of the first layer region of the upper layer over the lower layer. Then, when the first layer region of the upper layer with 3 μm thickness was formed, the RF glow discharge was stopped and the flow of the gas into the deposition chamber 1001 was interrupted by closing the flow-out valves 1041, 1042 and 1045, and the auxiliary valve 1018, thereby completing the formation of the first layer region of the upper layer.

Then, for forming the second layer region of the upper layer, the flow-out valves 1041 and 1042, and the auxiliary valve 1018 were gradually opened to flow SiH<sub>4</sub> gas and H<sub>2</sub> gas through the gas discharge aperture 1009 of the gas introduction pipe 1008 into the deposition chamber 1001. In this case, respective mass flow controllers 1021 and 1022 were adjusted so that the SiH<sub>4</sub> gas flow rate was 300 SCCM and H<sub>2</sub> flow rate was 300 SCCM. The pressure in the deposition chamber 1001 was controlled to 0.5 Torr by adjusting the opening of the main valve 1016 while observing the vacuum meter 1017. Then, RF power was introduced into the deposition chamber 1001 through the radio frequency matching box 1012 while setting the power of the RF power source (not illustrated) to 15 mW/cm<sup>3</sup>, to cause the RF glow discharge and start the formation of the second layer region on the first layer region of the upper layer. Then, when the second layer region of the upper layer with 20  $\mu$ m thickness was formed, the RF glow discharge was stopped and the flow of the gas into the deposition chamber 1001 was interrupted by closing the flow-out valves 1041 and 1042, and the auxiliary valve 1018, thereby completing the formation of the second layer region of the upper layer.

Then, for forming the third layer region of the upper layer, the flow-out valves 1041 and 1043, and the auxiliary valve 1018 were gradually opened to flow SiH<sub>4</sub> gas and CH<sub>4</sub> gas through the gas discharge aperture 1009 of the gas introduction pipe 1008 into the deposition chamber 1001. In this case, respective mass flow controllers 1021 and 1023 were adjusted so that the SiH<sub>4</sub> gas flow rate was 50 SCCM and CH<sub>4</sub> flow rate was 500 SCCM. The pressure in the deposition chamber 1001 was controlled to 0.4 Torr by adjusting the opening of the main valve 1016 while observing the vacuum meter 1017. Then, RF power was introduced into the deposition chamber 1001 through the radio frequency matching box 1012 while setting the power of the RF power source (not illustrated) to 10 mW/cm<sup>3</sup>, to cause the RF glow discharge and start the formation of the third layer region on the second layer region of the upper layer. Then, when the third layer region of the upper layer with 0.5  $\mu$ m thickness was formed, the RF glow discharge was stopped and the flow of the gas into the deposition chamber 1001 was interrupted by closing the flow-out valves 1041 and 1043, and the auxiliary valve 1018, thereby completing the formation of the third layer region of the upper layer.

The conditions for preparing the light receiving member for use in electrophotography described above are shown in Table 1.

It will be apparent that all of the flow-out valves other than those required for forming the respective layers were completely closed and, for avoiding the respective gases from remaining in the deposition chamber 1001 and in the pipeways from the flow-out valves 1041-1047 to the deposition chamber 1001, the flow-out valves 1041-1047 were closed, the auxiliary valve 1018 was opened and, further, the main valve was fully opened thereby evacuating the inside of the system once to a high vacuum degree as required.

Further, for forming the layer uniformly during this layer formation, the cylindrical aluminum support 1005 was rotated at a desired speed by a driving device not illustrated.

#### COMPARATIVE EXAMPLE 1

A light receiving member for use in electrophotography was prepared under the same preparation conditions as those in Example 1 except for not using H<sub>2</sub> gas upon forming the lower layer. The conditions for preparing the light receiving member for use in electrophotography are shown in Table 2.

The light receiving members for use in electrophotography thus prepared in Example 1 and Comparative Example 1 were set respectively to an electrophotographic apparatus, i.e., a copying machine NP-7550 manufactured by Canon Inc. and modified for experimental use and, when several electrophotographic properties were checked under various conditions.

It was found that both of the light receiving member for use in electrophotography has much excellent charging power.

Then, when the number of dots as the image characteristics were compared, it was found that the number of dots, particularly, the number of dots with less than 0.1 mm diameter of the light receiving member for use in electrophotography of Example 1 was less than  $\frac{1}{3}$  of that of the light receiving member for use in electrophotography in Comparative Example 1. In addition, for comparing the "coarse image", when the image density was measured for circular regions each of 0.05 mm diameter assumed as one unit at 100 points and the scattering in the image density was evaluated, it was found that the scattering in the light receiving member for use in electrophotography of Example 1 was less than  $\frac{1}{3}$  for that of the light receiving member for use in electrophotography in Comparative Example 1, and the light receiving member for use in electrophotography of Example 1 was excellent over the light receiving member for use in Electrophotography of Comparative Example 1 in view of the visual observation.

In addition, for comparing the occurrence of image defects and the peeling of the light receiving layer due to impactive mechanical pressure applied for a relatively short period of time to the light receiving member for use in electrophotography, when stainless steel balls of 3.5 mm diameter were fallen freely from the vertical height of 30 cm above the surface of the light receiving member for use in electrophotography and abutted against the surface of the light receiving member for use in electrophotography, to thereby measure the frequency of occurrence for cracks in the light receiving layer, it was found that the rate of occurrence in the light receiving member for use in electrophotography of Example 1 was less than  $\frac{3}{5}$  for that in the light receiving member for use in electrophotography of Comparative Example 1.

As has been described above, the light receiving member for use in electrophotography of Example 1 was superior to the light receiving member for use in electrophotography of Comparative Example 1.

#### EXAMPLE 2

A light receiving member for use in electrophotography was prepared in the same manner as in Example 1 except for changing the way of varying AlCl<sub>3</sub>/He gas flow rate in the lower layer, under the preparation conditions shown in Table 3 and, when evaluated in the same manner, satisfactory improvement was obtained to the dots, coarse image and peeling in the same manner as in Example 1.

## EXAMPLE 3

A light receiving member for use in electrophotography was prepared in the same manner as in Example 1 except for not using CH<sub>4</sub> gas in the upper layer of Example 1, under the preparation conditions shown in Table 4 and, when evaluated in the same manner, satisfactory improvement was obtained to the dots, coarse image and peeling in the same manner as in Example 1.

## EXAMPLE 4

A light receiving member for use in electrophotography was prepared in the same manner as in Example 1 except for replacing PH<sub>3</sub>/H<sub>2</sub> gas cylinder with He gas (99.9999% purity) cylinder and N<sub>2</sub> gas cylinder with NO gas (99.9% purity) cylinder in Example 1, and replacing H<sub>2</sub> gas with He gas and, further, using NO gas in the upper layer, under the preparation conditions shown in Table 5 and, when evaluated in the same manner, satisfactory improvement was obtained to the dots, coarse image and peeling in the same manner as in Example 1.

## EXAMPLE 5

A light receiving member for use in electrophotography was prepared in the same manner as in Example 1 except for replacing PH<sub>3</sub>/H<sub>2</sub> gas cylinder with Ar gas (99.9999% purity) cylinder and, further replacing N<sub>2</sub> gas cylinder with NH<sub>3</sub> gas (99.999% purity) cylinder in Example 1, replacing H<sub>2</sub> gas with Ar gas and replacing CH<sub>4</sub> gas with NH<sub>3</sub> gas in the upper layer, under the preparation conditions shown in Table 6 and, when evaluated in the same manner, satisfactory improvement was obtained to the dots, coarse image and peeling in the same manner as in Example 1.

## EXAMPLE 6

A light receiving member for use in electrophotography was prepared in the same manner as in Example 1 by further using PH<sub>3</sub>/H<sub>2</sub> gas in the upper layer, under the preparation conditions shown in Table 7 and, when evaluated in the same manner, satisfactory improvement was obtained to dots, coarse image and peeling in the same manner as in Example 1.

## EXAMPLE 7

A light receiving member for use in electrophotography was prepared in the same manner as in Example 1 by replacing N<sub>2</sub> gas cylinder with SiF<sub>4</sub> gas (99.999% purity) cylinder in Example 1, and, further using B<sub>2</sub>H<sub>6</sub>/H<sub>2</sub>, SiF<sub>4</sub> gas in the upper layer, under the preparation conditions shown in Table 8 and, when evaluated in the same manner, satisfactory improvement was obtained to dots, coarse image and peeling in the same manner as in Example 1.

## EXAMPLE 8

A light receiving member for use in electrophotography was prepared in the same manner as in Example 1 by further using PH<sub>3</sub>/H<sub>2</sub> gas and N<sub>2</sub> gas in the upper layer, under the preparation conditions shown in Table 9 and, when evaluated in the same manner, satisfactory improvement was obtained to dots, coarse image and peeling in the same manner as in Example 1.

## EXAMPLE 9

A light receiving member for use in electrophotography was prepared in the same manner as in Example 1

except for replacing CH<sub>4</sub> gas cylinder with C<sub>2</sub>H<sub>2</sub> gas (99.9999% purity) cylinder and N<sub>2</sub> gas cylinder with NO gas cylinder in Example 1, replacing CH<sub>4</sub> gas with C<sub>2</sub>H<sub>4</sub> gas, and further using NO gas in the upper layer, under the preparation conditions shown in Table 10 and, when evaluated in the same manner, satisfactory improvement was obtained to the dots, coarse image and peeling in the same manner as in Example 1.

## EXAMPLE 10

A light receiving member for use in electrophotography was prepared in the same manner as in Example 1, under the preparation conditions shown in Table 11 and, when evaluated in the same manner, satisfactory improvement was obtained to the dots, coarse image and peeling in the same manner as in Example 1.

## EXAMPLE 11

A light receiving member for use in electrophotography was prepared in the same manner as in Example 1 by replacing the N<sub>2</sub> gas cylinder with a NH<sub>3</sub> gas (99.999% purity) cylinder in Example 1, and replacing CH gas with NH<sub>3</sub> gas in the upper layer, under the preparation conditions shown in Table 12 and, when evaluated in the same manner, satisfactory improvement was obtained to the dots, coarse image and peeling in the same manner as in Example 1.

## EXAMPLE 12

A light receiving member for use in electrophotography was prepared in the same manner as in Example 6 by further replacing N<sub>2</sub> gas cylinder with SiF<sub>4</sub> gas cylinder in Example 6, and, further, using SiF<sub>4</sub> gas in the upper layer, under the preparation conditions shown in Table 13 and, when evaluated in the same manner, satisfactory improvement was obtained to dots, coarse image and peeling in the same manner as in Example 6.

## EXAMPLE 13

A light receiving member for use in electrophotography was prepared in the same manner as in Example 9 by further using B<sub>2</sub>H<sub>6</sub>/H<sub>2</sub> gas and Si<sub>2</sub>H<sub>6</sub> gas (99.99% purity) in the upper layer, under the preparation conditions shown in Table 14 and, when evaluated in the same manner, satisfactory improvement was obtained to dots, coarse image and peeling in the same manner as in Example 9.

## EXAMPLE 14

A light receiving member for use in electrophotography was prepared in the same manner as in Example 11 by using PH<sub>3</sub>/H<sub>2</sub> gas in the upper layer, under the preparation conditions shown in Table 15 and, when evaluated in the same manner, satisfactory improvement was obtained to dots, coarse image and peeling in the same manner as in Example 11.

## EXAMPLE 15

A light receiving member for use in electrophotography was prepared in the same manner as in Example 1 by further replacing N<sub>2</sub> gas cylinder with GeH<sub>4</sub> gas (99.999% purity) cylinder and further using GeH<sub>4</sub> gas in the upper layer, under the preparation conditions shown in Table 16 and, when evaluated in the same manner, satisfactory improvement was obtained to dots, coarse image and peeling in the same manner as in Example 1.

## EXAMPLE 16

A light receiving member for use in electrophotography was prepared in the same manner as in Example 1 by changing the outer diameter of the cylindrical aluminum support to 80 mm in Example 1, under the preparation conditions shown in Table 17 and, when evaluated in the same manner as in Example 1, except for using an electrophotographic apparatus, i.e., a copying machine NP-9030 manufactured by Canon Inc. and modified for the experimental use, satisfactory improvement was obtained to the dots, coarse image and peeling in the same manner as in Example 1.

## EXAMPLE 17

A light receiving member for use in electrophotography was prepared in the same manner as in Example 1 by changing the outer diameter of the cylindrical aluminum support to 60 mm in Example 1, under the preparation conditions shown in Table 18 and, when evaluated in the same manner as in Example 1, except for using an electrophotographic apparatus, i.e., a copying machine NP-150Z manufactured by Canon Inc. and modified for the experimental use, satisfactory improvement was obtained to the dots, coarse image and peeling in the same manner as in Example 1.

## EXAMPLE 18

A light receiving member for use in electrophotography was prepared in the same manner as in Example 1 by changing the outer diameter of the cylindrical aluminum support to 30 mm in Example 1, under the preparation conditions shown in Table 19 and, when evaluated in the same manner as in Example 1, except for using an electrophotographic apparatus, i.e., a copying machine FC-5 manufactured by Canon Inc. and modified for the experimental use, satisfactory improvement was obtained to the dots, coarse image and peeling in the same manner as in Example 1.

## EXAMPLE 19

A light receiving member for use in electrophotography was prepared in the same manner as in Example 1 by changing the outer diameter of the cylindrical aluminum support to 15 mm in Example 1, under the preparation conditions shown in Table 20, and evaluated in the same manner as in Example 1 except for using an electrophotographic apparatus, manufactured for experimental use, satisfactory improvement was obtained to the dots, coarse image and peeling in the same manner as in Example 1.

## EXAMPLE 20

A light sensitive member for use in electrophotography was prepared, under the same preparation conditions as those in Example 16 by using a cylindrical aluminum support applied with mirror-finishing fabrication in Example 16 and further machined into a cross sectional shape of:  $a=25$   $\mu\text{m}$ ,  $b=0.8$   $\mu\text{m}$  as shown in FIG. 38 by a diamond point tool and, when evaluated in the same manner as in Example 16, satisfactory improvement was obtained to, the dots, coarse image and peeling in the same manner as in Example 16.

## EXAMPLE 21

A light receiving member for use in electrophotography was prepared, under the same preparation conditions as those in Example 16 using a cylindrical alumi-

num support applied with mirror-finish fabrication and subsequently applied with a so-called surface dimpling of causing a number of hit pits to the surface of the cylindrical aluminum support by the exposure to a plurality of dropping bearing balls to form into a cross sectional shape of:  $c=50$   $\mu\text{m}$  and  $d=1$   $\mu\text{m}$  as shown in FIG. 39 and, when evaluated in the same manner as in Example 16, satisfactory improvement was obtained for the dots, coarse image and peeling in the same as in Example 16.

## EXAMPLE 22

A light receiving member for use in electrophotography having an upper layer comprising poly-Si(H, X) was prepared in the same manner as in Example 9 by using a cylindrical aluminum support heated to a temperature of 500° C., under the preparation conditions as shown in Table 21 and, when evaluated in the same manner, satisfactory improvement was obtained to dots, coarse image and peeling in the same manner as in Example 9.

## EXAMPLE 23

A light receiving member for use in electrophotography according to this invention was formed by microwave (hereinafter simply referred to as "uW") glow discharge decomposition:

A production apparatus for the light receiving member for use in photography by the uW glow discharge decomposition shown in FIG. 41 was used, in which a decomposition device 1100 for use in the uW glow discharge decomposition shown in FIG. 40 was used instead of the deposition device 1000 in the production apparatus of RF glow discharge decomposition shown in FIG. 37, and it was connected with a raw material gas supply device 1020.

In the figure, a cylindrical aluminum support 1107 had 108 mm of outer diameter and mirror-finished surface.

At first, in the same manner as in Example 1, the inside of the deposition chamber 1101 and the gas pipeways was evacuated such that the pressure in the deposition chamber 1101 was  $5 \times 10^{-6}$  Torr.

Then, in the same manner as in Example 1, the respective gases were introduced in the mass flow controllers 1021-1027. In this case, however, a SiF<sub>4</sub> gas cylinder was used in place of the N<sub>2</sub> gas cylinder.

Further, the cylindrical aluminum support 1107 disposed in the deposition chamber 1101 was heated to a temperature of 250° C. by a heater not illustrated.

After the preparation for the film formation was thus completed, each of the lower and the upper layers was formed on the cylindrical aluminum support 1107. The lower layer was formed by gradually opening the flow-out valves 1041, 1042 and 1047 and the auxiliary valve 1018, thereby flowing the SiH<sub>4</sub> gas, H<sub>2</sub> gas and AlCl<sub>3</sub>/He gas through the gas discharge aperture not illustrated of the gas introduction pipe 1110 into a plasma generation region 1109. In this case, the gas flow rate was controlled by each of the mass flow controllers 1021, 1022 and 1027 such that SiH<sub>4</sub> gas flow rate was 150 SCCM, H<sub>2</sub> gas flow rate was 20 SCCM and AlCl<sub>3</sub> gas flow rate was 400 SCCM. The pressure in the deposition chamber 1101 was set to 0.6 mTorr by adjusting the opening of the main valve not illustrated while observing the vacuum meter not illustrated. Then, uW power was introduced by way of a wave guide portion 1103 and a dielectric window 1102 into a plasma genera-

tion region 1109 by setting the power for a uW power source not illustrated to  $0.5 \text{ mW/cm}^3$ , to cause uW glow discharge and start the formation of the lower layer on the cylindrical aluminum support 1107. The mass flow controllers 1021, 1022 and 1027 were controlled such that the SiH<sub>4</sub> gas flow rate remained at a constant rate of 150 SCCM, the H<sub>2</sub> gas flow rate was increased at a constant ratio from 20 SCCM to 500 SCCM, the AlCl<sub>3</sub>/He gas flow rate was reduced at a constant ratio from 400 SCCM to 80 SCCM for the 0.01  $\mu\text{m}$  on the support side, while reduced at a constant ratio from 80 SCCM to 50 SCCM for 0.01  $\mu\text{m}$  on the side of the upper layer during formation of the lower layer. When the lower layer of 0.02  $\mu\text{m}$  thickness was formed, the uW glow discharge was stopped, the flow-out valves 1041, 1042, 1047 and the auxiliary valve 1018 were closed to interrupt the flow of the gas into the plasma generation region 1109 thereby completing the formation of the lower layer.

Then, for forming the first layer region of the upper layer, the flow-out valves 1041, 1042 and 1045, and the auxiliary valve 1018 were gradually opened to flow SiH<sub>4</sub> gas, H<sub>2</sub> gas, B<sub>2</sub>H<sub>6</sub>/H<sub>2</sub> through the gas discharge aperture not illustrated of the gas introduction pipe 1110 into the plasma generation space 1109. In this case, respective mass flow controllers 1021, 1022 and 1025 were adjusted so that SiH<sub>4</sub> gas flow rate was 100 SCCM, H<sub>2</sub> gas flow rate was 500 SCCM and B<sub>2</sub>H<sub>6</sub>/H<sub>2</sub> gas flow rate was 200 ppm to SiH<sub>4</sub> gas flow rate. The pressure in the deposition chamber 1101 was controlled to 0.5 mTorr. Then, RF power was introduced into the plasma generation chamber 1109 while setting the power of RF power source (not illustrated) to  $0.5 \text{ mW/cm}^3$ , to cause uW glow discharge and start the formation of the first layer region of the upper layer over the lower layer. Then, the first layer region of 3  $\mu\text{m}$  thickness of the upper layer was formed.

Then, for forming the second layer region of the upper layer, the flow-out valves 1041, 1042 and 1046, and the auxiliary valve 1018 were gradually opened to flow SiH<sub>4</sub> gas, H<sub>2</sub> gas and SiF<sub>4</sub> gas through the gas discharge aperture not illustrated of the gas introduction pipe 1110 into the plasma generation space 1109. In this case, respective mass flow controllers 1021, 1022 and 1026 were adjusted so that the SiH<sub>4</sub> gas flow rate was 700 SCCM, H<sub>2</sub> gas flow rate was 500 SCCM and SiF<sub>4</sub> gas flow rate was 30 SCCM. The pressure in the deposition chamber 1101 was controlled to 0.5 mTorr. Then, the power of a uW power source (not illustrated) was set to  $0.5 \text{ mW/cm}^3$ , to cause uW glow discharge in the plasma generation region 1109 and form the second layer region with 20  $\mu\text{m}$  thickness of the upper layer on the first layer region of the upper layer.

Then, for forming the third layer region of the upper layer, the flow-out valves 1041 and 1043 and the auxiliary valve 1018 were gradually opened to flow SiH<sub>4</sub> gas and CH<sub>4</sub> gas through the gas discharge aperture not illustrated of the gas introduction pipe 1110 into the plasma generation space 1109. In this case, respective mass flow controllers 1021 and 1023 were adjusted so that the SiH<sub>4</sub> gas flow rate was 150 SCCM and CH<sub>4</sub> gas flow rate was 500 SCCM. The pressure in the deposition chamber 1101 was controlled to 0.3 mTorr. Then, the power of a uW power source (not illustrated) was set to  $0.5 \text{ mW/cm}^3$ , to cause uW glow discharge in the plasma generation region 1109 and the third layer region with 0.5  $\mu\text{m}$  thickness of the upper layer was formed on the second layer region of the upper layer.

The conditions for preparing the light receiving member for use in electrophotography described above are shown in Table 22.

When the light receiving member for use in electrophotography was evaluated in the same manner in Example 1, improvement was obtained to the dots, coarse image and peeling in the same manner as in Example 1.

#### EXAMPLE 24

10 A light receiving member for use in electrophotography was prepared in the same manner as in Example 1, under the preparation conditions shown in Table 23 and, when evaluated in the same manner, satisfactory improvement was obtained to the dots, coarse image 15 and peeling in the same manner as in Example 1.

#### EXAMPLE 25

20 A light receiving member for use in electrophotography was prepared in the same manner as in Example 1, under the preparation conditions shown in Table 24 and, when evaluated in the same manner, satisfactory improvement was obtained to the dots, coarse image 25 and peeling in the same manner as in Example 1.

#### EXAMPLE 26

25 A light receiving member for use in electrophotography was prepared in the same manner as in Example 1, under the preparation conditions shown in Table 25 and, when evaluated in the same manner, satisfactory improvement was obtained to the dots, coarse image 30 and peeling in the same manner as in Example 1.

#### EXAMPLE 27

35 A light receiving member for use in electrophotography was prepared in the same manner as in Example 1, under the preparation conditions shown in Table 26 and, when evaluated in the same manner, satisfactory improvement was obtained to the dots, coarse image 40 and peeling in the same manner as in Example 6.

#### EXAMPLE 28

45 A light receiving member for use in electrophotography was prepared in the same manner as in Example 9, under the preparation conditions shown in Table 27 and, when evaluated in the same manner, satisfactory improvement was obtained to the dots, coarse image 50 and peeling in the same manner as in Example 9.

#### EXAMPLE 29

50 A light receiving member for use in electrophotography was prepared in the same manner as in Example 11, under the preparation conditions shown in Table 28 and, when evaluated in the same manner, satisfactory improvement was obtained to the dots, coarse image 55 and peeling in the same manner as in Example 11.

#### EXAMPLE 30

55 A light receiving member for use in electrophotography was prepared in the same manner as in Example 1, under the preparation conditions shown in Table 29 and, when evaluated in the same manner, satisfactory improvement was obtained to the dots, coarse image 60 and peeling in the same manner as in Example 1.

#### EXAMPLE 31

65 A light receiving member for use in electrophotography was prepared in the same manner as in Example 1, under the preparation conditions shown in Table 30

and, when evaluated in the same manner, satisfactory improvement was obtained to the dots, coarse image and peeling in the same manner as in Example 1.

#### EXAMPLE 32

A light receiving member for use in electrophotography was prepared in the same manner as in Example 6, under the preparation conditions shown in Table 31 and, when evaluated in the same manner, satisfactory improvement was obtained to the dots, coarse image 10 and peeling in the same manner as in Example 6.

#### EXAMPLE 33

A light receiving member for use in electrophotography was prepared in the same manner as in Example 1, under the preparation conditions shown in Table 32 and, when evaluated in the same manner, satisfactory improvement was obtained to the dots, coarse image 15 and peeling in the same manner as in Example 1.

#### EXAMPLE 34

A light receiving member for use in electrophotography was prepared in the same manner as in Example 1 by further using  $B_2H_6$  gas upon forming the lower layer 20 in Example 1, under the preparation conditions as 25 shown in Table 33.

#### COMPARATIVE EXAMPLE 2

A light receiving member for use in electrophotography was prepared under the same preparation conditions as those in Example 34 except for not using  $B_2H_6/H_2$  gas upon forming the lower layer. The conditions for preparing the light receiving member for use in 30 electrophotography are shown in Table 34.

The light receiving members for use in electrophotography thus prepared in Example 34 and Comparative Example 2 were set respectively to an electrophotographic apparatus, i.e., a copying machine NP-7550 manufactured by Canon Inc. and modified for experimental use and, when several electrophotographic 40 properties were checked under various conditions.

It was found that both of the light receiving member for use in electrophotography has much excellent charging power.

Then, when the number of dots as the image characteristics were compared, it was found that the number of dots, particularly, the number of dots with less than 0.1 mm diameter of the light receiving member for use in electrophotography of Example 24 was less than  $\frac{1}{4}$  of that of the light receiving member for use in electrophotography in Comparative Example 2. In addition, for comparing the "coarse image", when the image density was measured for circular regions each of 0.05 mm diameter assumed as one unit at 100 points and the scattering in the image density was evaluated, it was found that the scattering in the light receiving member for use in electrophotography of Example 24 was less than  $\frac{1}{2}$  for that of the light receiving member for use in electrophotography in Comparative Example 2, and the light receiving member for use in electrophotography of 50 Example 1 was excellent over the light receiving member for use in Electrophotography of Comparative Example 2 in view of the visual observation.

In addition, for comparing the occurrence of image defects and the peeling of the light receiving layer due 60 to impactive mechanical pressure applied for a relatively short period of time to the light receiving member for use in electrophotography, when stainless steel

balls of 3.5 mm diameter were fallen freely from the vertical height of 30 cm above the surface of the light receiving member for use in electrophotography and abutted against the surface of the light receiving member for use in electrophotography, to thereby measure the frequency of occurrence for cracks in the light receiving layer, it was found that the rate of occurrence in the light receiving member for use in electrophotography of Example 24 was less than 3/5 for that in the light receiving member for use in electrophotography of Comparative Example 2.

As has been described above, the light receiving member for use in electrophotography of Example 24 was superior to the light receiving member for use in electrophotography of Comparative Example 2.

#### EXAMPLE 35

A light receiving member for use in electrophotography was prepared in the same manner as in Example 34 20 except for changing the way of varying  $AlCl_3/He$  gas flow rate in the lower layer, under the preparation conditions shown in Table 35 and, when evaluated in the same manner, satisfactory improvement was obtained to the dots, coarse image and peeling in the same manner as in Example 34.

#### EXAMPLE 36

A light receiving member for use in electrophotography was prepared in the same manner as in Example 35 except for not using  $CH_4$  gas in the upper layer of Example 34, under the preparation conditions shown in Table 36 and, when evaluated in the same manner, satisfactory improvement was obtained to the dots, coarse image and peeling in the same manner as in Example 34.

#### EXAMPLE 37

A light receiving member for use in electrophotography was prepared in the same manner as in Example 34 except for replacing  $PH_3/H_2$  gas cylinder with He gas (99.9999% purity) cylinder and  $N_2$  gas cylinder with NO gas (99.9% purity) cylinder, replacing  $H_2$  gas with  $SiF_4$  gas cylinder and using NO gas,  $SiF_4$  gas in Example 34, under the preparation conditions shown in Table 5 and, when evaluated in the same manner, satisfactory improvement was obtained to the dots, coarse image and peeling in the same manner as in Example 34.

#### EXAMPLE 38

A light receiving member for use in electrophotography was prepared in the same manner as in Example 1 except for replacing  $PH_3/H_2$  gas cylinder with Ar gas (99.9999% purity) cylinder and, further replacing  $N_2$  gas cylinder with  $NH_3$  gas (99.999% purity) cylinder in Example 34, and replacing  $H_2$  gas with Ar gas and replacing  $CH_4$  gas with  $NH_3$  gas in the upper layer, under the preparation conditions shown in Table 38 and, when evaluated in the same manner, satisfactory improvement was obtained to the dots, coarse image and peeling in the same manner as in Example 34.

#### EXAMPLE 39

A light receiving member for use in electrophotography was prepared in the same manner as in Example 34 by further using  $PH_3/H_2$  gas in the upper layer, under the preparation conditions shown in Table 39 and, when evaluated in the same manner, satisfactory improvement was obtained to dots, coarse image and peeling in the same manner as in Example 34.

## EXAMPLE 40

A light receiving member for use in electrophotography was prepared in the same manner as in Example 34 by replacing N<sub>2</sub> gas cylinder with SiF<sub>4</sub> gas (99.999% purity) cylinder in Example 34, and, further using B<sub>2</sub>H<sub>6</sub>/H<sub>2</sub>, SiF<sub>4</sub> gas in the upper layer, under the preparation conditions shown in Table 40 and, when evaluated in the same manner, satisfactory improvement was obtained to dots, coarse image and peeling in the same manner as in Example 34.

## EXAMPLE 41

A light receiving member for use in electrophotography was prepared in the same manner as in Example 34 by further using PH<sub>3</sub>/H<sub>2</sub> gas and N<sub>2</sub> gas in the upper layer, under the preparation conditions shown in Table 41 and, when evaluated in the same manner, satisfactory improvement was obtained to dots, coarse image and peeling in the same manner as in Example 34.

## EXAMPLE 42

A light receiving member for use in electrophotography was prepared in the same manner as in Example 34 except for replacing CH<sub>4</sub> gas cylinder with C<sub>2</sub>H<sub>2</sub> gas (99.9999% purity) cylinder and N<sub>2</sub> gas cylinder with NO gas cylinder in Example 34, and using NO gas in the upper layer, under the preparation conditions shown in Table 42 and, when evaluated in the same manner, satisfactory improvement was obtained to the dots, coarse image and peeling in the same manner as in Example 34.

## EXAMPLE 43

A light receiving member for use in electrophotography was prepared in the same manner as in Example 34, under the preparation conditions shown in Table 11 in the upper layer and, when evaluated in the same manner, satisfactory improvement was obtained to the dots, coarse image and peeling in the same manner as in Example 34.

## EXAMPLE 44

A light receiving member for use in electrophotography was prepared in the same manner as in Example 34 by replacing N<sub>2</sub> gas cylinder with NH<sub>3</sub> gas (99.999% purity) cylinder in Example 34, and replacing CH gas with NH<sub>3</sub> gas in the upper layer, under the preparation conditions shown in Table 44 and, when evaluated in the same manner, satisfactory improvement was obtained to the dots, coarse image and peeling in the same manner as in Example 34.

## EXAMPLE 45

A light receiving member for use in electrophotography was prepared in the same manner as in Example 39 by replacing N<sub>2</sub> gas cylinder with SiF<sub>4</sub> gas cylinder in Example 39, and, further, using SiF<sub>4</sub> gas in the upper layer, under the preparation conditions shown in Table 45 and, when evaluated in the same manner, satisfactory improvement was obtained to dots, coarse image and peeling in the same manner as in Example 39.

## EXAMPLE 46

A light receiving member for use in electrophotography was prepared in the same manner as in Example 42 by further using B<sub>2</sub>H<sub>6</sub>/H<sub>2</sub> gas and Si<sub>2</sub>H<sub>6</sub> gas (99.99% purity) in the upper layer, under the preparation conditions shown in Table 46 and, when evaluated in the

5

same manner, satisfactory improvement was obtained to dots, coarse image and peeling in the same manner as in Example 42.

## EXAMPLE 47

A light receiving member for use in electrophotography was prepared in the same manner as in Example 44 by using PH<sub>3</sub>/H<sub>2</sub> gas in the upper layer, under the preparation conditions shown in Table 47 and, when evaluated in the same manner, satisfactory improvement was obtained to dots, coarse image and peeling in the same manner as in Example 44.

## EXAMPLE 48

A light receiving member for use in electrophotography was prepared in the same manner as in Example 34 by further replacing N<sub>2</sub> gas cylinder with GeH<sub>4</sub> gas (99.999% purity) cylinder and further using GeH<sub>4</sub> gas in the upper layer, under the preparation conditions shown in Table 48 and, when evaluated in the same manner, satisfactory improvement was obtained to dots, coarse image and peeling in the same manner as in Example 34.

## EXAMPLE 49

A light receiving member for use in electrophotography was prepared in the same manner as in Example 34 by changing the outer diameter of the cylindrical aluminum support to 80 mm in Example 34, under the preparation conditions shown in Table 49 and, when evaluated in the same manner as in Example 34, except for using an electrophotographic apparatus, i.e., a copying machine NP-9030 manufactured by Canon Inc. and modified for the experimental use, satisfactory improvement was obtained to the dots, coarse image and peeling in the same manner as in Example 34.

## EXAMPLE 50

A light receiving member for use in electrophotography was prepared in the same manner as in Example 34 by changing the outer diameter of the cylindrical aluminum support to 60 mm in Example 34, under the preparation conditions shown in Table 50 and, when evaluated in the same manner as in Example 34, except for using an electrophotographic apparatus, i.e., a copying machine NP-150Z manufactured by Canon Inc. and modified for the experimental use, satisfactory improvement was obtained to the dots, coarse image and peeling in the same manner as in Example 34.

## EXAMPLE 51

A light receiving member for use in electrophotography was prepared in the same manner as in Example 34 by changing the outer diameter of the cylindrical aluminum support to 30 mm in Example 34, under the preparation conditions shown in Table 51 and, when evaluated in the same manner as in Example 34, except for using an electrophotographic apparatus, i.e., a copying machine FC-5 manufactured by Canon Inc. and modified for the experimental use, satisfactory improvement was obtained to the dots, coarse image and peeling in the same manner as in Example 34.

## EXAMPLE 52

A light receiving member for use in electrophotography was prepared in the same manner as in Example 34 by changing the outer diameter of the cylindrical aluminum support to 15 mm in Example 34, under the prepa-

10

15

20

30

35

40

45

50

55

60

65

ration conditions shown in Table 52, and evaluated in the same manner as in Example 1 except for using an electrophotographic apparatus, manufactured for experimental use, satisfactory improvement was obtained to the dots, coarse image and peeling in the same manner as in Example 34.

#### EXAMPLE 53

A light sensitive member for use in electrophotography was prepared, under the same preparation conditions as those in Example 49 by using a cylindrical aluminum support applied with mirror-finish fabrication in Example 49 and further machined into a cross sectional shape of:  $a=25$   $\mu\text{m}$ ,  $b=0.8$   $\mu\text{m}$  as shown in FIG. 38 by a diamond point tool and, when evaluated in the same manner as in Example 49, satisfactory improvement was obtained to, the dots, coarse image and peeling in the same manner as in Example 49.

#### EXAMPLE 54

A light receiving member for use in electrophotography was prepared, under the same preparation conditions as those in Example 49 using a cylindrical aluminum support applied with mirror-finish fabrication and subsequently applied with a so-called surface dimpling of causing a number of hit pits to the surface of the cylindrical aluminum support by the exposure to a plurality of dropping bearing balls to form into a cross sectional shape of:  $c=50$   $\mu\text{m}$  and  $d=1$   $\mu\text{m}$  as shown in FIG. 39 and, when evaluated in the same manner as in Example 49, satisfactory improvement was obtained for the dots, coarse image and peeling in the same manner as in Example 49.

#### EXAMPLE 55

A light receiving member for use in electrophotography having an upper layer comprising poly-Si(H, X) was prepared in the same manner as in Example 42 by using a cylindrical aluminum support heated to a temperature of 500° C., under the preparation conditions as shown in Table 53 and, when evaluated in the same manner, satisfactory improvement was obtained to dots, coarse image and peeling in the same manner as in Example 42.

#### EXAMPLE 56

A light receiving member for use in electrophotography was formed by microwave glow discharge decomposition in the same manner as in Example 23 by further using  $\text{H}_2\text{S}$  gas and  $\text{B}_2\text{H}_6$  gas under the preparation conditions shown in Table 54 upon forming the low layer in Example 23.

When the light receiving member for use in electrophotography was evaluated in the same manner as in Example 34, improvement was obtained to the dots, coarse image and peeling in the same manner as in Example 34.

#### EXAMPLE 57

A light receiving member for use in electrophotography was prepared in the same manner as in Example 42, under the preparation conditions shown in Table 55 and, when evaluated in the same manner, satisfactory improvement was obtained to the dots, coarse image and peeling in the same manner as in Example 42.

#### EXAMPLE 58

A light receiving member for use in electrophotography was prepared in the same manner as in Example 43, under the preparation conditions shown in Table 56 and, when evaluated in the same manner, satisfactory improvement was obtained to the dots, coarse image and peeling in the same manner as in Example 43.

#### EXAMPLE 59

A light receiving member for use in electrophotography was prepared in the same manner as in Example 44, under the preparation conditions shown in Table 57 and, when evaluated in the same manner, satisfactory improvement was obtained to the dots, coarse image and peeling in the same manner as in Example 44.

#### EXAMPLE 60

A light receiving member for use in electrophotography was prepared in the same manner as in Example 45, under the preparation conditions shown in Table 58 and, when evaluated in the same manner, satisfactory improvement was obtained to the dots, coarse image and peeling in the same manner as in Example 45.

#### EXAMPLE 61

A light receiving member for use in electrophotography was prepared in the same manner as in Example 46, under the preparation conditions shown in Table 59 and, when evaluated in the same manner, satisfactory improvement was obtained to the dots, coarse image and peeling in the same manner as in Example 41.

#### EXAMPLE 62

A light receiving member for use in electrophotography was prepared in the same manner as in Example 47, under the preparation conditions shown in Table 60 and, when evaluated in the same manner, satisfactory improvement was obtained to the dots, coarse image and peeling in the same manner as in Example 47.

#### EXAMPLE 63

A light receiving member for use in electrophotography was prepared in the same manner as in Example 37, under the preparation conditions shown in Table 61 and, when evaluated in the same manner, satisfactory improvement was obtained to the dots, coarse image and peeling in the same manner as in Example 37.

#### EXAMPLE 64

A light receiving member for use in electrophotography was prepared in the same manner as in Example 39, under the preparation conditions shown in Table 62 and, when evaluated in the same manner, satisfactory improvement was obtained to the dots, coarse image and peeling in the same manner as in Example 39.

#### EXAMPLE 65

A light receiving member for use in electrophotography was prepared in the same manner as in Example 45, under the preparation conditions shown in Table 63 and, when evaluated in the same manner, satisfactory improvement was obtained to the dots, coarse image and peeling in the same manner as in Example 45.

#### EXAMPLE 66

A light receiving member for use in electrophotography was prepared in the same manner as in Example 64,

under the preparation conditions shown in Table 64 and, when evaluated in the same manner, satisfactory improvement was obtained to the dots, coarse image and peeling in the same manner as in Example 64.

#### EXAMPLE 67

A light receiving member for use in electrophotography was prepared in the same manner as in Example 1 by further using NO gas upon forming the lower layer in Example 1, under the preparation conditions as shown in Table 65.

#### COMPARATIVE EXAMPLE 3

A light receiving member for use in electrophotography was prepared under the same preparation conditions as those in Example 67 except for not using H<sub>2</sub> gas and NO gas upon forming the lower layer. The conditions for preparing the light receiving member for use in electrophotography are shown in Table 66.

The light receiving members for use in electrophotography thus prepared in Example 67 and Comparative Example 3 were set respectively to an electrophotographic apparatus, i.e., a copying machine NP-7550 manufactured by Canon Inc. and modified for experimental use and, when several electrophotographic properties were checked under various conditions.

It was found that both of the light receiving member for use in electrophotography had much excellent charging power.

Then, when the number of dots as the image characteristics were compared, it was found that the number of dots, particularly, the number of dots with less than 0.1 mm diameter of the light receiving member for use in electrophotography of Example 67 was less than  $\frac{3}{4}$  of that of the light receiving member for use in electrophotography in Comparative Example 3. In addition, for comparing the "coarse image", when the image density was measured for circular regions each of 0.05 mm diameter assumed as one unit at 100 points and the scattering in the image density was evaluated, it was found that the scattering in the light receiving member for use in electrophotography of Example 67 was less than  $\frac{1}{2}$  for that of the light receiving member for use in electrophotography in Comparative Example 3, and the light receiving member for use in electrophotography of Example 67 was excellent over the light receiving member for use in Electrophotography of Comparative Example 3 in view of the visual observation.

In addition, for comparing the occurrence of image defects and the peeling of the light receiving layer due to impactive mechanical pressure applied for a relatively short period of time to the light receiving member for use in electrophotography, when stainless steel balls of 3.5 mm diameter were fallen freely from the vertical height of 30 cm above the surface of the light receiving member for use in electrophotography and abutted against the surface of the light receiving member for use in electrophotography, to thereby measure the frequency of occurrence for cracks in the light receiving layer, it was found that the rate of occurrence in the light receiving for use in electrophotography of Example 67 was less than 2/5 for that in the light receiving member for use in electrophotography of Comparative Example 3.

As has been described above, the light receiving member for use in electrophotography of Example 67 was superior to the light receiving member for use in electrophotography of Comparative Example 3.

#### EXAMPLE 68

A light receiving member for use in electrophotography was prepared in the same manner as in Example 67 except for changing the way of varying AlCl<sub>3</sub>/He gas flow rate in the lower layer, under the preparation conditions shown in Table 67 and, when evaluated in the same manner, satisfactory improvement was obtained to the dots, coarse image and peeling in the same manner as in Example 67.

#### EXAMPLE 69

A light receiving member for use in electrophotography was prepared in the same manner as in Example 67 except for not using CH<sub>4</sub> gas in the upper layer of Example 67, under the preparation conditions shown in Table 68 and, when evaluated in the same manner, satisfactory improvement was obtained to the dots, coarse image and peeling in the same manner as in Example 67.

#### EXAMPLE 70

A light receiving member for use in electrophotography was prepared in the same manner as in Example 67 except for replacing PH<sub>3</sub>/H<sub>2</sub> gas cylinder with He gas (99.999% purity) cylinder and NO gas and N<sub>2</sub> gas from a not illustrated cylinder in Example 67, under the preparation conditions shown in Table 69 and, when evaluated in the same manner, satisfactory improvement was obtained to the dots, coarse image and peeling in the same manner as in Example 67.

#### EXAMPLE 71

A light receiving member for use in electrophotography was prepared in the same manner as in Example 67 except for replacing PH<sub>3</sub>/H<sub>2</sub> gas cylinder with Ar gas (99.999% purity) cylinder and, further replacing NO gas cylinder with NH<sub>3</sub> gas (99.999% purity) cylinder, replacing AlCl<sub>3</sub>/He gas with Al(CH<sub>3</sub>)<sub>3</sub>/He gas (99.99% purity) and using CH<sub>4</sub> gas in the lower layer in Example 67, replacing H<sub>2</sub> gas with Ar gas and CH<sub>4</sub> gas with NH<sub>3</sub> gas in the upper layer, under the preparation conditions shown in Table 70 and, when evaluated in the same manner, satisfactory improvement was obtained to the dots, coarse image and peeling in the same manner as in Example 67.

#### EXAMPLE 72

A light receiving member for use in electrophotography was prepared in the same manner as in Example 67 by further using PH<sub>3</sub>/H<sub>2</sub> gas in the upper layer, under the preparation conditions shown in Table 71 and, when evaluated in the same manner, satisfactory improvement was obtained to dots, coarse image and peeling in the same manner as in Example 67.

#### EXAMPLE 73

A light receiving member for use in electrophotography was prepared in the same manner as in Example 67 by further using PH<sub>3</sub>/H<sub>2</sub> gas, not illustrated SiF<sub>4</sub> gas (99.999% purity) cylinder in Example 67, under the preparation conditions shown in Table 8 and, when evaluated in the same manner, satisfactory improvement was obtained to dots, coarse image and peeling in the same manner as in Example 67.

#### EXAMPLE 74

A light receiving member for use in electrophotography was prepared in the same manner as in Example 67

by further using  $\text{CH}_4$  gas,  $\text{B}_2\text{H}_6/\text{H}_2$  gas and not illustrated  $\text{H}_2\text{S}$  gas (99.9% purity) in the lower layer, and using  $\text{PH}_3/\text{H}_2$  gas and  $\text{N}_2$  gas in the upper layer, under the preparation conditions shown in Table 73 and, when evaluated in the same manner, satisfactory improvement was obtained to dots, coarse image and peeling in the same manner as in Example 67.

#### EXAMPLE 75

A light receiving member for use in electrophotography was prepared in the same manner as in Example 67 except for replacing  $\text{CH}_4$  gas cylinder with  $\text{C}_2\text{H}_2$  gas (99.999% purity) cylinder in Example 67 and replacing  $\text{CH}_4$  gas with  $\text{C}_2\text{H}_4$  gas, and further using  $\text{NO}$  gas in the upper layer, under the preparation conditions shown in Table 74 and, when evaluated in the same manner, satisfactory improvement was obtained to the dots, coarse image and peeling in the same manner as in Example 67.

#### EXAMPLE 76

A light receiving member for use in electrophotography was prepared in the same manner as in Example 67, under the preparation conditions shown in Table 75 and, when evaluated in the same manner, satisfactory improvement was obtained to the dots, coarse image and peeling in the same manner as in Example 67.

#### EXAMPLE 77

A light receiving member for use in electrophotography was prepared in the same manner as in Example 67 by replacing the  $\text{CH}_4$  gas cylinder with a  $\text{NH}_3$  gas (99.999% purity) cylinder in Example 67, and replacing  $\text{CH}_4$  gas with  $\text{NH}_3$  gas in the upper layer, under the preparation conditions shown in Table 76 and, when evaluated in the same manner, satisfactory improvement was obtained to the dots, coarse image and peeling in the same manner as in Example 67.

#### EXAMPLE 78

A light receiving member for use in electrophotography was prepared in the same manner as in Example 72 by further using  $\text{SiF}_4$  gas in the upper layer in Example 72, under the preparation conditions shown in Table 77 and, when evaluated in the same manner, satisfactory improvement was obtained to dots, coarse image and peeling in the same manner as in Example 72.

#### EXAMPLE 79

A light receiving member for use in electrophotography was prepared in the same manner as in Example 75 by further using  $\text{B}_2\text{H}_6/\text{H}_2$  gas and  $\text{Si}_2\text{H}_6$  gas in the upper layer, under the preparation conditions shown in Table 78 and, when evaluated in the same manner, satisfactory improvement was obtained to dots, coarse image and peeling in the same manner as in Example 75.

#### EXAMPLE 80

A light receiving member for use in electrophotography was prepared in the same manner as in Example 77 by further using  $\text{PH}_3/\text{H}_2$  gas in the upper layer, under the preparation conditions shown in Table 75 and, when evaluated in the same manner, satisfactory improvement was obtained to dots, coarse image and peeling in the same manner as in Example 77.

#### EXAMPLE 81

A light receiving member for use in electrophotography was prepared in the same manner as in Example 67

10

by further replacing  $\text{B}_2\text{H}_6/\text{H}_2$  gas cylinder with  $\text{GeH}_4$  gas (99.999% purity) cylinder in Example 67 and further using  $\text{GeH}_4$  gas in the upper layer, under the preparation conditions shown in Table 80 and, when evaluated in the same manner, satisfactory improvement was obtained to dots, coarse image and peeling in the same manner as in Example 67.

15

20

#### EXAMPLE 82

A light receiving member for use in electrophotography was prepared in the same manner as in Example 67 by changing the outer diameter of the cylindrical aluminum support to 80 mm in Example 67, under the preparation conditions shown in Table 81 and, when evaluated in the same manner as in Example 67, except for using an electrophotographic apparatus, i.e., a copying machine NP-9030 manufactured by Canon Inc. and modified for the experimental use, satisfactory improvement was obtained to the dots, coarse image and peeling in the same manner as in Example 67.

#### EXAMPLE 83

A light receiving member for use in electrophotography was prepared in the same manner as in Example 67 by changing the outer diameter of the cylindrical aluminum support to 60 mm in Example 67, under the preparation conditions shown in Table 82 and, when evaluated in the same manner as in Example 67, except for using an electrophotographic apparatus, i.e., a copying machine NP-150Z manufactured by Canon Inc. and modified for the experimental use, satisfactory improvement was obtained to the dots, coarse image and peeling in the same manner as in Example 67.

#### EXAMPLE 84

A light receiving member for use in electrophotography was prepared in the same manner as in Example 67 by changing the outer diameter of the cylindrical aluminum support to 30 mm in Example 67, under the preparation conditions shown in Table 83 and, when evaluated in the same manner as in Example 67, except for using an electrophotographic apparatus, i.e., a copying machine FC-5 manufactured by Canon Inc. and modified for the experimental use, satisfactory improvement was obtained to the dots, coarse image and peeling in the same manner as in Example 67.

#### EXAMPLE 85

A light receiving member for use in electrophotography was prepared in the same manner as in Example 67 by changing the outer diameter of the cylindrical aluminum support to 15 mm in Example 67, under the preparation conditions shown in Table 84, and evaluated in the same manner as in Example 67 except for using an electrophotographic apparatus, manufactured for experimental use, satisfactory improvement was obtained to the dots, coarse image and peeling in the same manner as in Example 67.

#### EXAMPLE 86

A light sensitive member for use in electrophotography was prepared, under the same preparation conditions as those in Example 82 by using a cylindrical aluminum support applied with mirror-finishing fabrication in Example 82 and further machined into a cross sectional shape of:  $a=25 \mu\text{m}$ ,  $b=0.8 \mu\text{m}$  as shown in FIG. 38 by a diamond point tool and, when evaluated in the same manner as in Example 82, satisfactory im-

60

65

provement was obtained to, the dots, coarse image and peeling in the same manner as in Example 82.

#### EXAMPLE 87

A light receiving member for use in electrophotography was prepared, under the same preparation conditions as those in Example 82 using a cylindrical aluminum support applied with mirror-finish fabrication and subsequently applied with a so-called surface dimpling of causing a number of hit pits to the surface of the cylindrical aluminum support by the exposure to a plurality of dropping bearing balls to form into a cross sectional shape of:  $c=50 \mu\text{m}$  and  $d=1 \mu\text{m}$  as shown in FIG. 39 and, when evaluated in the same manner as in Example 82, satisfactory improvement was obtained for the dots, coarse image and peeling in the same as in Example 82.

#### EXAMPLE 88

A light receiving member for use in electrophotography having an upper layer comprising poly-Si(H, X) was prepared in the same manner as in Example 75 by using a cylindrical aluminum support heated to a temperature of 500° C., under the preparation conditions as shown in Table 85 and, when evaluated in the same manner, satisfactory improvement was obtained to dots, coarse image and peeling in the same manner as in Example 75.

#### EXAMPLE 89

A light receiving member for use in electrophotography was formed by microwave glow discharge decomposition in the same manner as in Example 23, further using NO gas and B<sub>2</sub>H<sub>6</sub> gas upon forming lower layer under the preparation conditions shown in Table 86.

When the light receiving member for use in electrophotography was evaluated in the same manner in Example 67 improvement was obtained to the dots, coarse image and peeling in the same manner as in Example 67.

#### EXAMPLE 90

A light receiving member for use in electrophotography was prepared in the same manner as in Example 75, under the preparation conditions shown in Table 87 and, when evaluated in the same manner, satisfactory improvement was obtained to the dots, coarse image and peeling in the same manner as in Example 75.

#### EXAMPLE 91

A light receiving member for use in electrophotography was prepared in the same manner as in Example 76, under the preparation conditions shown in Table 88 and, when evaluated in the same manner, satisfactory improvement was obtained to the dots, coarse image and peeling in the same manner as in Example 76.

#### EXAMPLE 92

A light receiving member for use in electrophotography was prepared in the same manner as in Example 77, under the preparation conditions shown in Table 89 and, when evaluated in the same manner, satisfactory improvement was obtained to the dots, coarse image and peeling in the same manner as in Example 77.

#### EXAMPLE 93

A light receiving member for use in electrophotography was prepared in the same manner as in Example 78, under the preparation conditions shown in Table 90

and, when evaluated in the same manner, satisfactory improvement was obtained to the dots, coarse image and peeling in the same manner as in Example 78.

#### EXAMPLE 94

A light receiving member for use in electrophotography was prepared in the same manner as in Example 79, under the preparation conditions shown in Table 91 and, when evaluated in the same manner, satisfactory improvement was obtained to the dots, coarse image and peeling in the same manner as in Example 79.

#### EXAMPLE 95

A light receiving member for use in electrophotography was prepared in the same manner as in Example 80, under the preparation conditions shown in Table 92 and, when evaluated in the same manner, satisfactory improvement was obtained to the dots, coarse image and peeling in the same manner as in Example 80.

#### EXAMPLE 96

A light receiving member for use in electrophotography was prepared in the same manner as in Example 70, under the preparation conditions shown in Table 93 and, when evaluated in the same manner, satisfactory improvement was obtained to the dots, coarse image and peeling in the same manner as in Example 70.

#### EXAMPLE 97

30 A light receiving member for use in electrophotography was prepared in the same manner as in Example 72, under the preparation conditions shown in Table 94 and, when evaluated in the same manner, satisfactory improvement was obtained to the dots, coarse image and peeling in the same manner as in Example 72.

#### EXAMPLE 98

40 A light receiving member for use in electrophotography was prepared in the same manner as in Example 78, under the preparation conditions shown in Table 75 and, when evaluated in the same manner, satisfactory improvement was obtained to the dots, coarse image and peeling in the same manner as in Example 78.

#### EXAMPLE 99

A light receiving member for use in electrophotography was prepared in the same manner as in Example 97, under the preparation conditions shown in Table 96 and, when evaluated in the same manner, satisfactory improvement was obtained to the dots, coarse image and peeling in the same manner as in Example 97.

#### EXAMPLE 100

55 A light receiving member for use in electrophotography was prepared in the same manner as in Example 1 by further using SiF<sub>4</sub> gas upon forming the lower layer in Example 97, under the preparation conditions as shown in Table 33.

#### COMPARATIVE EXAMPLE 4

A light receiving member for use in electrophotography was prepared under the same preparation conditions as those in Example 100 except for not using SiF<sub>4</sub> gas and H<sub>2</sub> gas upon forming the lower layer. The conditions for preparing the light receiving member for use in electrophotography are shown in Table 98.

The light receiving members for use in electrophotography thus prepared in Example 100 and Compara-

tive Example 4 were set respectively to an electrophotographic apparatus, i.e., a copying machine NP-7550 manufactured by Canon Inc. and modified for experimental use and several electrophotographic properties were checked under various conditions.

It was found that both of the light receiving member for use in electrophotography had much excellent charging power. Then, when the number of dots as the image characteristics were compared, it was found that the number of dots, particularly, the number of dots with less than 0.1 mm diameter of the light receiving member for use in electrophotography of Example 100 was less than  $\frac{1}{2}$  of that of the light receiving member for use in electrophotography in Comparative Example 4. In addition, for comparing the "coarse image", when the image density was measured for circular regions each of 0.05 mm diameter assumed as one unit at 100 points and the scattering in the image density was evaluated, it was found that the scattering in the light receiving member for use in electrophotography of Example 100 was less than  $\frac{1}{2}$  for that of the light receiving member for use in electrophotography in Comparative Example 4, and the light receiving member for use in electrophotography of Example 100 was excellent over the light receiving member for use in Electrophotography of Comparative Example 4 in view of the visual observation.

In addition, for comparing the occurrence of image defects and the peeling of the light receiving layer due to impactive mechanical pressure applied for a relatively short period of time to the light receiving member for use in electrophotography, when stainless steel balls of 3.5 mm diameter were fallen freely from the vertical height of 30 cm above the surface of the light receiving member for use in electrophotography and abutted against the surface of the light receiving member for use in electrophotography, to thereby measure the frequency of occurrence for cracks in the light receiving layer, it was found that the rate of occurrence in the light receiving member for use in electrophotography of Example 100 was less than 2/5 for that in the light receiving member for use in electrophotography of Comparative Example 4.

As has been described above, the light receiving member for use in electrophotography of Example 100 was superior to the light receiving member for use in electrophotography of Comparative Example 4.

#### EXAMPLE 101

A light receiving member for use in electrophotography was prepared in the same manner as in Example 100 except for further using NO gas, B<sub>2</sub>H<sub>6</sub>/H<sub>2</sub> gas and changing the way of varying AlCl<sub>3</sub>/He gas flow rate in the lower layer of Example 100, under the preparation conditions shown in Table 89 and, when evaluated in the same manner, satisfactory improvement was obtained to the dots, coarse image and peeling in the same manner as in Example 100.

#### EXAMPLE 102

A light receiving member for use in electrophotography was prepared in the same manner as in Example 100 except for not using CH<sub>4</sub> gas in the upper layer of Example 100, under the preparation conditions shown in Table 100 and, when evaluated in the same manner, satisfactory improvement was obtained to the dots, coarse image and peeling in the same manner as in Example 100.

#### EXAMPLE 103

A light receiving member for use in electrophotography was prepared in the same manner as in Example 100 except for further using N<sub>2</sub> gas (99.9999% purity) and He gas (99.9999% purity) in Example 100, under the preparation conditions shown in Table 101 and, when evaluated in the same manner, satisfactory improvement was obtained to the dots, coarse image and peeling in the same manner as in Example 100.

#### EXAMPLE 104

A light receiving member for use in electrophotography was prepared in the same manner as in Example 100 except for replacing AlCl<sub>3</sub> with Al(CH<sub>3</sub>)<sub>3</sub> (99.99% purity) in Example 100, and further replacing SiF<sub>4</sub> gas cylinder with Ar gas (99.9999% purity) cylinder and NO gas cylinder with NH<sub>3</sub> gas (99.999% purity) cylinder in the upper layer, under the preparation conditions shown in Table 102 and, when evaluated in the same manner, satisfactory improvement was obtained to the dots, coarse image and peeling in the same manner as in Example 100.

#### EXAMPLE 105

A light receiving member for use in electrophotography was prepared in the same manner as in Example 100 by further using PH<sub>3</sub>/H<sub>2</sub> gas in the upper layer, under the preparation conditions shown in Table 103 and, when evaluated in the same manner, satisfactory improvement was obtained to dots, coarse image and peeling in the same manner as in Example 100.

#### EXAMPLE 106

A light receiving member for use in electrophotography was prepared in the same manner as in Example 100 by using PHF<sub>5</sub> gas diluted with He gas (99.999% purity, referred to simply as "PF<sub>5</sub>/He") cylinder in the lower layer of Example 100, and, further using B<sub>2</sub>H<sub>6</sub>/H<sub>2</sub>, SiF<sub>4</sub> gas in the upper layer, under the preparation conditions shown in Table 104 and, when evaluated in the same manner, satisfactory improvement was obtained to dots, coarse image and peeling in the same manner as in Example 100.

#### EXAMPLE 107

A light receiving member for use in electrophotography was prepared in the same manner as in Example 100 by using H<sub>2</sub>S gas in the lower layer of Example 100 and further using PH<sub>3</sub>/H<sub>2</sub> gas and N<sub>2</sub> gas in the upper layer, under the preparation conditions shown in Table 105 and, when evaluated in the same manner, satisfactory improvement was obtained to dots, coarse image and peeling in the same manner as in Example 100.

#### EXAMPLE 108

A light receiving member for use in electrophotography was prepared in the same manner as in Example 100 except for replacing CH<sub>4</sub> gas cylinder with C<sub>2</sub>H<sub>2</sub> gas (99.9999% purity) cylinder in Example 100, under the preparation conditions shown in Table 106 and, when evaluated in the same manner, satisfactory improvement was obtained to the dots, coarse image and peeling in the same manner as in Example 100.

#### EXAMPLE 109

A light receiving member for use in electrophotography was prepared in the same manner as in Example

100, by using  $\text{BF}_3$  gas diluted with He gas (99.999% purity, hereinafter simply referred to as " $\text{BF}_3/\text{He}$  gas"), under the preparation conditions shown in Table 17 and, when evaluated in the same manner, satisfactory improvement was obtained to the dots, coarse image and peeling in the same manner as in Example 100.

#### EXAMPLE 110

A light receiving member for use in electrophotography was prepared in the same manner as in Example 100 by replacing the NO gas cylinder with  $\text{NH}_3$  gas cylinder in Example 100, and replacing  $\text{CH}_4$  gas with  $\text{NH}_3$  gas in the upper layer, under the preparation conditions shown in Table 108 and, when evaluated in the same manner, satisfactory improvement was obtained to the dots, coarse image and peeling in the same manner as in Example 100.

#### EXAMPLE 111

A light receiving member for use in electrophotography was prepared in the same manner as in Example 105 by further using  $\text{SiF}_4$  gas in the upper layer of Example 105, under the preparation conditions shown in Table 109 and, when evaluated in the same manner, satisfactory improvement was obtained to dots, coarse image and peeling in the same manner as in Example 105.

#### EXAMPLE 112

A light receiving member for use in electrophotography was prepared in the same manner as in Example 100 by using  $\text{Si}_2\text{H}_6$  gas (99.99% purity) instead of  $\text{SiF}_4$  gas in the lower layer and further using  $\text{B}_2\text{H}_6/\text{H}_2$  gas and  $\text{Si}_2\text{H}_6$  gas (99.99% purity) in the upper layer, under the preparation conditions shown in Table 110 and, when evaluated in the same manner, satisfactory improvement was obtained to dots, coarse image and peeling in the same manner as in Example 100.

#### EXAMPLE 113

A light receiving member for use in electrophotography was prepared in the same manner as in Example 100 by using  $\text{Si}_2\text{H}_6$  gas in the lower layer and using  $\text{PH}_3/\text{H}_2$  gas in the upper layer, under the preparation conditions shown in Table 111 and, when evaluated in the same manner, satisfactory improvement was obtained to dots, coarse image and peeling in the same manner as in Example 100.

#### EXAMPLE 114

A light receiving member for use in electrophotography was prepared in the same manner as in Example 100 by replacing NO gas cylinder with  $\text{GeH}_4$  gas (99.999% purity) cylinder and further using  $\text{GeH}_4$  gas in the upper layer, under the preparation conditions shown in Table 112 and, when evaluated in the same manner, satisfactory improvement was obtained to dots, coarse image and peeling in the same manner as in Example 100.

#### EXAMPLE 115

A light receiving member for use in electrophotography was prepared in the same manner as in Example 100 by changing the outer diameter of the cylindrical aluminum support to 80 mm in Example 100, under the preparation conditions shown in Table 113 and, when evaluated in the same manner as in Example 100, except for using an electrophotographic apparatus, i.e., a copying machine NP-9030 manufactured by Canon Inc. and modified for the experimental use, satisfactory improvement was obtained to the dots, coarse image and peeling in the same manner as in Example 100.

ment was obtained to the dots, coarse image and peeling in the same manner as in Example 100.

#### EXAMPLE 116

A light receiving member for use in electrophotography was prepared in the same manner as in Example 100 by changing the outer diameter of the cylindrical aluminum support to 60 mm in Example 100, under the preparation conditions shown in Table 114 and, when evaluated in the same manner as in Example 1, except for using an electrophotographic apparatus, i.e., a copying machine NP-150Z manufactured by Canon Inc. and modified for the experimental use, satisfactory improvement was obtained to the dots, coarse image and peeling in the same manner as in Example 100.

#### EXAMPLE 117

A light receiving member for use in electrophotography was prepared in the same manner as in Example 100 by changing the outer diameter of the cylindrical aluminum support to 30 mm in Example 100, under the preparation conditions shown in Table 115 and, when evaluated in the same manner as in Example 100, except for using an electrophotographic apparatus, i.e., a copying machine FC-5 manufactured by Canon Inc. and modified for the experimental use, satisfactory improvement was obtained to the dots, coarse image and peeling in the same manner as in Example 100.

#### EXAMPLE 118

A light receiving member for use in electrophotography was prepared in the same manner as in Example 100 by changing the outer diameter of the cylindrical aluminum support to 15 mm in Example 100, under the preparation conditions shown in Table 116, and evaluated in the same manner as in Example 100 except for using an electrophotographic apparatus, manufactured for experimental use, satisfactory improvement was obtained to the dots, coarse image and peeling in the same manner as in Example 100.

#### EXAMPLE 119

A light sensitive member for use in electrophotography was prepared, under the same preparation conditions as those in Example 115 by using a cylindrical aluminum support applied with mirror-finishing fabrication in Example 115 and further machined into a cross sectional shape of:  $a=25 \mu\text{m}$ ,  $b=0.8 \mu\text{m}$  as shown in FIG. 38 by a diamond point tool and, when evaluated in the same manner as in Example 115, satisfactory improvement was obtained to the dots, coarse image and peeling in the same manner as in Example 115.

#### EXAMPLE 120

A light receiving member for use in electrophotography was prepared, under the same preparation conditions as those in Example 115 using a cylindrical aluminum support applied with mirror-finish fabrication and subsequently applied with a so-called surface dimpling of causing a number of hit pits to the surface of the cylindrical aluminum support by the exposure to a plurality of dropping bearing balls to form into a cross sectional shape of:  $c=50 \mu\text{m}$  and  $d=1 \mu\text{m}$  as shown in FIG. 39 and, when evaluated in the same manner as in Example 16, satisfactory improvement was obtained for the dots, coarse image and peeling in the same as in Example 115.

## EXAMPLE 121

A light receiving member for use in electrophotography having an upper layer comprising poly-Si(H, X) was prepared in the same manner as in Example 108 by using a cylindrical aluminum support heated to a temperature of 500° C., under the preparation conditions as shown in Table 117 and, when evaluated in the same manner, satisfactory improvement was obtained to dots, coarse image and peeling in the same manner as in Example 108.

## EXAMPLE 122

A light receiving member for use in electrophotography was formed by microwave glow discharge decomposition in the same manner as in Example 1, by further using SiF<sub>4</sub> gas, NO gas and B<sub>2</sub>H<sub>6</sub> gas upon forming the upper layer in Example 23, under the preparing conditions shown in Table 118.

When the light receiving member for use in electrophotography was evaluated in the same manner in Example 100, improvement was obtained to the dots, coarse image and peeling in the same manner as in Example 1.

## EXAMPLE 123

A light receiving member for use in electrophotography was prepared in the same manner as in Example 108, under the preparation conditions shown in Table 119 and, when evaluated in the same manner, satisfactory improvement was obtained to the dots, coarse image and peeling in the same manner as in Example 108.

## EXAMPLE 124

A light receiving member for use in electrophotography was prepared in the same manner as in Example 108, under the preparation conditions shown in Table 120 and, when evaluated in the same manner, satisfactory improvement was obtained to the dots, coarse image and peeling in the same manner as in Example 109.

## EXAMPLE 125

A light receiving member for use in electrophotography was prepared in the same manner as in Example 110, under the preparation conditions shown in Table 121 and, when evaluated in the same manner, satisfactory improvement was obtained to the dots, coarse image and peeling in the same manner as in Example 110.

## EXAMPLE 126

A light receiving member for use in electrophotography was prepared in the same manner as in Example 111, under the preparation conditions shown in Table 122 and, when evaluated in the same manner, satisfactory improvement was obtained to the dots, coarse image and peeling in the same manner as in Example 111.

## EXAMPLE 127

A light receiving member for use in electrophotography was prepared in the same manner as in Example 127, under the preparation conditions shown in Table 123 and, when evaluated in the same manner, satisfactory improvement was obtained to the dots, coarse

image and peeling in the same manner as in Example 112.

## EXAMPLE 128

A light receiving member for use in electrophotography was prepared in the same manner as in Example 113, under the preparation conditions shown in Table 124 and, when evaluated in the same manner, satisfactory improvement was obtained to the dots, coarse image and peeling in the same manner as in Example 113.

## EXAMPLE 129

A light receiving member for use in electrophotography was prepared in the same manner as in Example 103, under the preparation conditions shown in Table 125 and, when evaluated in the same manner, satisfactory improvement was obtained to the dots, coarse image and peeling in the same manner as in Example 103.

## EXAMPLE 130

A light receiving member for use in electrophotography was prepared in the same manner as in Example 105, under the preparation conditions shown in Table 126 and, when evaluated in the same manner, satisfactory improvement was obtained to the dots, coarse image and peeling in the same manner as in Example 105.

## EXAMPLE 131

A light receiving member for use in electrophotography was prepared in the same manner as in Example 111, under the preparation conditions shown in Table 127 and, when evaluated in the same manner, satisfactory improvement was obtained to the dots, coarse image and peeling in the same manner as in Example 111.

## EXAMPLE 132

A light receiving member for use in electrophotography was prepared in the same manner as in Example 130, under the preparation conditions shown in Table 128 and, when evaluated in the same manner, satisfactory improvement was obtained to the dots, coarse image and peeling in the same manner as in Example 130.

## EXAMPLE 133

A light receiving member for use in electrophotography was prepared in the same manner as in Example 1 by further using GeH<sub>4</sub> gas upon forming the lower layer in Example 1, under the preparation conditions as shown in Table 129.

## COMPARATIVE EXAMPLE 5

A light receiving member for use in electrophotography was prepared under the same preparation conditions as those in Example 133 except for not using GeH<sub>4</sub> gas and H<sub>2</sub> gas upon forming the lower layer. The conditions for preparing the light receiving member for use in electrophotography are shown in Table 130.

The light receiving members for use in electrophotography thus prepared in Example 133 and Comparative Example 5 were set respectively to an electrophotographic apparatus, i.e., a copying machine NP-7550 manufactured by Canon Inc. and modified for experi-

mental use and several electrophotographic properties were checked under various conditions.

It was found that both of the light receiving member for use in electrophotography had much excellent charging power. Then, when the number of dots as the image characteristics were compared, it was found that the number of dots, particularly, the number of dots with less than 0.1 mm diameter of the light receiving member for use in electrophotography of Example 133 was less than 2/5 of that of the light receiving member for use in electrophotography in Comparative Example 5. In addition, for comparing the "coarse image", when the image density was measured for circular regions each of 0.05 mm diameter assumed as one unit at 100 points and the scattering in the image density was evaluated, it was found that the scattering in the light receiving member for use in electrophotography of Example 133 was less than  $\frac{1}{3}$  for that of the light receiving member for use in electrophotography in Comparative Example 5, and the light receiving member for use in electrophotography of Example 133 was excellent over the light receiving member for use in Electrophotography of Comparative Example 5 in view of the visual observation.

In addition, for comparing the occurrence of image defects and the peeling of the light receiving layer due to impactive mechanical pressure applied for a relatively short period of time to the light receiving member for use in electrophotography, when stainless steel balls of 3.5 mm diameter were fallen freely from the vertical height of 30 cm above the surface of the light receiving member for use in electrophotography and abutted against the surface of the light receiving member for use in electrophotography, to thereby measure the frequency of occurrence for cracks in the light receiving layer, it was found that the rate of occurrence in the light receiving member for use in electrophotography of Example 133 was less than 3/5 for that in the light receiving member for use in electrophotography of Comparative Example 5.

When the lower layer of the light receiving member for use in electrophotography of Example 133 was analyzed by using SIMS, it was found that the content of silicon atoms, hydrogen atoms and aluminum atoms along the layer thickness changed as desired.

As has been described above, the light receiving member for use in electrophotography of Example 133 was superior to the light receiving member for use in electrophotography of Comparative Example 133.

#### EXAMPLE 134

A light receiving member for use in electrophotography was prepared in the same manner as in Example 133 except for further using NO gas, B<sub>2</sub>H<sub>6</sub> gas and H<sub>2</sub> gas and changing the way of varying AlCl<sub>3</sub>/He gas flow rate in the lower layer of Example 133, under the preparation conditions shown in Table 131 and, when evaluated in the same manner, satisfactory improvement was obtained to the dots, coarse image and peeling in the same manner as in Example 33.

#### EXAMPLE 135

A light receiving member for use in electrophotography was prepared in the same manner as in Example 133 except for not using CH<sub>4</sub> gas in the upper layer of Example 133, under the preparation conditions shown in Table 132 and, when evaluated in the same manner, satisfactory improvement was obtained to the dots,

coarse image and peeling in the same manner as in Example 133.

#### EXAMPLE 136

5 A light receiving member for use in electrophotography was prepared in the same manner as in Example 133 except for using N<sub>2</sub> gas (99.9999% purity) and He gas (99.9999% purity) in Example 133, under the preparation conditions shown in Table 133 and, when evaluated 10 in the same manner, satisfactory improvement was obtained to the dots, coarse image and peeling in the same manner as in Example 133.

#### EXAMPLE 137

15 A light receiving member for use in electrophotography was prepared in the same manner as in Example 133 except for replacing AlCl<sub>3</sub> with Al(CH<sub>3</sub>)<sub>3</sub>(99.99% purity) in the lower layer of Example 133 and replacing SiF<sub>4</sub> gas cylinder Ar gas (99.9999% purity) cylinder and, further replacing NO gas cylinder with NH<sub>3</sub> gas (99.999% purity) cylinder in the upper layer, under the preparation conditions shown in Table 134 and, when evaluated 20 in the same manner, satisfactory improvement was obtained to the dots, coarse image and peeling in the same manner as in Example 133.

#### EXAMPLE 138

25 A light receiving member for use in electrophotography was prepared in the same manner as in Example 133 except for further using PH<sub>3</sub>/H<sub>2</sub> gas in the upper layer, under the preparation conditions shown in Table 135 and, when evaluated 30 in the same manner, satisfactory improvement was obtained to dots, coarse image and peeling in the same manner as in Example 133.

#### EXAMPLE 139

35 A light receiving member for use in electrophotography was prepared in the same manner as in Example 133 by using PF<sub>3</sub> gas diluted with He gas (99.999% purity, hereinafter simply referred to as "PF<sub>3</sub>/He") cylinder in the lower layer of Example 133, and, further using B<sub>2</sub>H<sub>6</sub>/H<sub>2</sub>, SiF<sub>4</sub> gas in the upper layer, under the preparation 40 conditions shown in Table 136 and, when evaluated in the same manner, satisfactory improvement was obtained to dots, coarse image and peeling in the same manner as in Example 133.

#### EXAMPLE 140

45 A light receiving member for use in electrophotography was prepared in the same manner as in Example 133 by using H<sub>2</sub>S gas (99.9% purity) in the lower layer of Example 133 and further using PH<sub>3</sub>/H<sub>2</sub> gas and N<sub>2</sub> gas in the upper layer, under the preparation conditions 50 shown in Table 137 and, when evaluated in the same manner as in Example 133, satisfactory improvement was obtained to dots, coarse image and peeling in the same manner as in Example 141.

#### EXAMPLE 141

55 A light receiving member for use in electrophotography was prepared in the same manner as in Example 138 except for replacing CH<sub>4</sub> gas cylinder with C<sub>2</sub>H<sub>2</sub> gas (99.9999% purity) cylinder in Example 139, under the preparation conditions shown in Table 138 and, when evaluated 60 in the same manner, satisfactory improvement was obtained to the dots, coarse image and peeling in the same manner as in Example 133.

## EXAMPLE 142

A light receiving member for use in electrophotography was prepared in the same manner as in Example 133, using  $\text{BF}_3$  gas diluted with  $\text{He}$  gas (99.999% purity, hereinafter simply referred to as "BF<sub>3</sub>/gas) in the lower layer of Example 133, under the preparation conditions shown in Table 133 and, when evaluated in the same manner, satisfactory improvement was obtained to the dots, coarse image and peeling in the same manner as in Example 133.

## EXAMPLE 143

A light receiving member for use in electrophotography was prepared in the same manner as in Example 133 by replacing  $\text{CH}_4$  gas cylinder with  $\text{NH}_3$  gas cylinder in Example 133, and replacing  $\text{CH}_4$  gas with  $\text{NH}_3$  gas in the upper layer, under the preparation conditions shown in Table 140 and, when evaluated in the same manner, satisfactory improvement was obtained to the dots, coarse image and peeling in the same manner as in Example 133.

## EXAMPLE 144

A light receiving member for use in electrophotography was prepared in the same manner as in Example 138 by further using  $\text{SiF}_4$  gas in the upper layer of Example 138, under the preparation conditions shown in Table 13 and, when evaluated in the same manner, satisfactory improvement was obtained to dots, coarse image and peeling in the same manner as in Example 138.

## EXAMPLE 145

A light receiving member for use in electrophotography was prepared in the same manner as in Example 133 by further using  $\text{B}_2\text{H}_6/\text{H}_2$  gas and  $\text{Si}_2\text{H}_6$  gas (99.99% purity) in the upper layer, under the preparation conditions shown in Table 142 and, when evaluated in the same manner, satisfactory improvement was obtained to dots, coarse image and peeling in the same manner as in Example 133.

## EXAMPLE 146

A light receiving member for use in electrophotography was prepared in the same manner as in Example 133 by using  $\text{Si}_2\text{F}_6$  gas in the lower layer and using  $\text{PH}_3/\text{H}_2$  gas in the upper layer, under the preparation conditions shown in Table 143 and, when evaluated in the same manner, satisfactory improvement was obtained to dots, coarse image and peeling in the same manner as in Example 133.

## EXAMPLE 147

A light receiving member for use in electrophotography was prepared in the same manner as in Example 133 by further using  $\text{GeH}_4$  gas in the upper layer of Example 133, under the preparation conditions shown in Table 144 and, when evaluated in the same manner, satisfactory improvement was obtained to dots, coarse image and peeling in the same manner as in Example 133.

## EXAMPLE 148

A light receiving member for use in electrophotography was prepared in the same manner as in Example 133 by changing the outer diameter of the cylindrical aluminum support to 80 mm in Example 133, under the preparation conditions shown in Table 145 and, when evaluated

in the same manner as in Example 133, except for using an electrophotographic apparatus, i.e., a copying machine NP-9030 manufactured by Canon Inc. and modified for the experimental use, satisfactory improvement was obtained to the dots, coarse image and peeling in the same manner as in Example 133.

## EXAMPLE 149

A light receiving member for use in electrophotography was prepared in the same manner as in Example 133 by changing the outer diameter of the cylindrical aluminum support to 60 mm in Example 133, under the preparation conditions shown in Table 146 and, when evaluated in the same manner as in Example 133, except for using an electrophotographic apparatus, i.e., a copying machine NP-150Z manufactured by Canon Inc. and modified for the experimental use, satisfactory improvement was obtained to the dots, coarse image and peeling in the same manner as in Example 133.

## EXAMPLE 150

A light receiving member for use in electrophotography was prepared in the same manner as in Example 133 by changing the outer diameter of the cylindrical aluminum support to 30 mm in Example 133, under the preparation conditions shown in Table 147 and, when evaluated in the same manner as in Example 133, except for using an electrophotographic apparatus, i.e., a copying machine FC-5 manufactured by Canon Inc. and modified for the experimental use, satisfactory improvement was obtained to the dots, coarse image and peeling in the same manner as in Example 133.

## EXAMPLE 151

A light receiving member for use in electrophotography was prepared in the same manner as in Example 133 by changing the outer diameter of the cylindrical aluminum support to 15 mm in Example 133, under the preparation conditions shown in Table 147, and evaluated in the same manner as in Example 1 except for using an electrophotographic apparatus, manufactured for experimental use, satisfactory improvement was obtained to the dots, coarse image and peeling in the same manner as in Example 133.

## EXAMPLE 152

A light sensitive member for use in electrophotography was prepared, under the same preparation conditions as those in Example 148 by using a cylindrical aluminum support applied with mirror-finishing fabrication in Example 148 and further machined into a cross sectional shape of:  $a=25 \mu\text{m}$ ,  $b=0.8 \mu\text{m}$  as shown in FIG. 38 by a diamond point tool and, when evaluated in the same manner as in Example 148, satisfactory improvement was obtained to the dots, coarse image and peeling in the same manner as in Example 148.

## EXAMPLE 153

A light receiving member for use in electrophotography was prepared, under the same preparation conditions as those in Example 148 using a cylindrical aluminum support applied with mirror-finish fabrication and subsequently applied with a so-called surface dimpling of causing a number of hit pits to the surface of the cylindrical aluminum support by the exposure to a plurality of dropping bearing balls to form into a cross sectional shape of:  $c=50 \mu\text{m}$  and  $d=1 \mu\text{m}$  as shown in FIG. 39 and, when evaluated in the same manner as in

Example 148, satisfactory improvement was obtained for the dots, coarse image and peeling in the same manner as in Example 148.

#### EXAMPLE 154

A light receiving member for use in electrophotography having an upper layer comprising poly-Si(H, X) was prepared in the same manner as in Example 141 by using a cylindrical aluminum support heated to a temperature of 500° C., under the preparation conditions as shown in Table 149 and, when evaluated in the same manner, satisfactory improvement was obtained to dots, coarse image and peeling in the same manner as in Example 141.

#### EXAMPLE 155

A light receiving member for use in electrophotography was formed by microwave glow discharge decomposition in the same manner as in Example 23, further using BeH<sub>4</sub> gas, B<sub>2</sub>H<sub>6</sub> gas, NO gas and SiF<sub>4</sub> gas, upon forming the lower layer in Example 23, under the preparing conditions shown in Table 150.

When the light receiving member for use in electrophotography was evaluated in the same manner in Example 133, improvement was obtained to the dots, coarse image and peeling in the same manner as in Example 133.

#### EXAMPLE 156

A light receiving member for use in electrophotography was prepared in the same manner as in Example 141, under the preparation conditions shown in Table 151 and, when evaluated in the same manner, satisfactory improvement was obtained to the dots, coarse image and peeling in the same manner as in Example 141.

#### EXAMPLE 157

A light receiving member for use in electrophotography was prepared in the same manner as in Example 142, under the preparation conditions shown in Table 152 and, when evaluated in the same manner, satisfactory improvement was obtained to the dots, coarse image and peeling in the same manner as in Example 142.

#### EXAMPLE 158

A light receiving member for use in electrophotography was prepared in the same manner as in Example 143, under the preparation conditions shown in Table 153 and, when evaluated in the same manner, satisfactory improvement was obtained to the dots, coarse image and peeling in the same manner as in Example 143.

#### EXAMPLE 159

A light receiving member for use in electrophotography was prepared in the same manner as in Example 144, under the preparation conditions shown in Table 154 and, when evaluated in the same manner, satisfactory improvement was obtained to the dots, coarse image and peeling in the same manner as in Example 144.

#### EXAMPLE 160

A light receiving member for use in electrophotography was prepared in the same manner as in Example 145, under the preparation conditions shown in Table

155 and, when evaluated in the same manner, satisfactory improvement was obtained to the dots, coarse image and peeling in the same manner as in Example 45.

#### EXAMPLE 161

5 A light receiving member for use in electrophotography was prepared in the same manner as in Example 146, under the preparation conditions shown in Table 156 and, when evaluated in the same manner, satisfactory improvement was obtained to the dots, coarse image and peeling in the same manner as in Example 146.

#### EXAMPLE 162

15 A light receiving member for use in electrophotography was prepared in the same manner as in Example 136, under the preparation conditions shown in Table 157 and, when evaluated in the same manner, satisfactory improvement was obtained to the dots, coarse image and peeling in the same manner as in Example 136.

#### EXAMPLE 163

20 A light receiving member for use in electrophotography was prepared in the same manner as in Example 138, under the preparation conditions shown in Table 158 and, when evaluated in the same manner, satisfactory improvement was obtained to the dots, coarse image and peeling in the same manner as in Example 138.

#### EXAMPLE 164

25 A light receiving member for use in electrophotography was prepared in the same manner as in Example 144, under the preparation conditions shown in Table 159 and, when evaluated in the same manner, satisfactory improvement was obtained to the dots, coarse image and peeling in the same manner as in Example 144.

#### EXAMPLE 165

30 A light receiving member for use in electrophotography was prepared in the same manner as in Example 163, under the preparation conditions shown in Table 160 and, when evaluated in the same manner, satisfactory improvement was obtained to the dots, coarse image and peeling in the same manner as in Example 163.

#### EXAMPLE 166

35 A light receiving member for use in electrophotography was prepared in the same manner as in Example 1 by further using Mg(C<sub>5</sub>H<sub>6</sub>)<sub>2</sub>/He gas B<sub>2</sub>H<sub>6</sub> gas upon forming the lower layer in Example 1, under the preparation conditions as shown in Table 161.

#### COMPARATIVE EXAMPLE 6

40 A light receiving member for use in electrophotography was prepared under the same preparation conditions as those in Example 166 except for not using H<sub>2</sub> and Mg(C<sub>5</sub>H<sub>6</sub>)<sub>2</sub>/He gas upon forming the lower layer. The conditions for preparing the light receiving member for use in electrophotography are shown in Table 162.

45 The light receiving members for use in electrophotography thus prepared in Example 166 and Comparative Example 6 were set respectively to an electrophotographic apparatus, i.e., a copying machine NP-7550

manufactured by Canon Inc. and modified for experimental use and several electrophotographic properties were checked under various conditions.

It was found that both of the light receiving member for use in electrophotography had much excellent charging power. Then, when the number of dots as the image characteristics were compared, it was found that the number of dots, particularly, the number of dots with less than 0.1 mm diameter of the light receiving member for use in electrophotography of Example 166 was less than  $\frac{1}{2}$  of that of the light receiving member for use in electrophotography in Comparative Example 6. In addition, for comparing the "coarse image", when the image density was measured for circular regions each of 0.05 mm diameter assumed as one unit at 100 points and the scattering in the image density was evaluated, it was found that the scattering in the light receiving member for use in electrophotography of Example 166 was less than  $\frac{1}{4}$  for that of the light receiving member for use in electrophotography in Comparative Example 6, and the light receiving member for use in electrophotography of Example 166 was excellent over the light receiving member for use in Electrophotography of Comparative Example 6 in view of the visual observation.

In addition, for comparing the occurrence of image defects and the peeling of the light receiving layer due to impactive mechanical pressure applied for a relatively short period of time to the light receiving member for use in electrophotography, when stainless steel 30 balls of 3.5 mm diameter were fallen freely from the vertical height of 30 cm above the surface of the light receiving member for use in electrophotography and abutted against the surface of the light receiving member for use in electrophotography, to thereby measure 35 the frequency of occurrence for cracks in the light receiving layer, it was found that the rate of occurrence in the light receiving member for use in electrophotography of Example 166 was less than  $\frac{1}{2}$  for that in the light receiving member for use in electrophotography of 40 Comparative Example 6.

When the lower layer of the light receiving member for use in electrophotography of Example 166 was analyzed by using SIMS, it was found that the content of silicon atoms, hydrogen atoms and aluminum atoms 45 along the layer thickness changed as desired.

As has been described above, the light receiving member for use in electrophotography of Example 166 was superior to the light receiving member for use in electrophotography of Comparative Example 6.

#### EXAMPLE 167

A light receiving member for use in electrophotography was prepared in the same manner as in Example 166 except for further using NO gas and  $\text{B}_2\text{H}_6/\text{H}_2$  gas, 55 changing the way of varying  $\text{AlCl}_3/\text{He}$  gas flow rate in the lower layer of Example 166, under the preparation conditions shown in Table 163 and, when evaluated in the same manner, satisfactory improvement was obtained to the dots, coarse image and peeling in the same 60 manner as in Example 166.

#### EXAMPLE 168

A light receiving member for use in electrophotography was prepared in the same manner as in Example 166 except for not using  $\text{CH}_4$  gas in the upper layer of Example 166, under the preparation conditions shown in Table 164 and, when evaluated in the same manner, 65

satisfactory improvement was obtained to the dots, coarse image and peeling in the same manner as in Example 166.

#### EXAMPLE 169

A light receiving member for use in electrophotography was prepared in the same manner as in Example 1 except for fur using  $\text{N}_2$  gas (99.9999% purity), He gas (99.9999% purity) and  $\text{SiF}_4$  gas from not illustrated cylinders in Example 166, under the preparation conditions shown in Table 165 and, when evaluated in the same manner, satisfactory improvement was obtained to the dots, coarse image and peeling in the same manner as in Example 166.

#### EXAMPLE 170

A light receiving member for use in electrophotography was prepared in the same manner as in Example 1 except for using  $\text{Al}(\text{CH}_3)_3$  instead of  $\text{AlCl}_3$  (99.99%, purity) and using further  $\text{CH}_4$  gas in the lower layer and replacing  $\text{SiF}_4$  gas cylinder with Ar gas (99.9999% purity) cylinder and, further replacing NO gas cylinder with  $\text{NH}_3$  gas (99.999% purity) cylinder in the upper layer of Example 166, under the preparation conditions shown in Table 166 and, when evaluated in the same manner, satisfactory improvement was obtained to the dots, coarse image and peeling in the same manner as in Example 166.

#### EXAMPLE 171

A light receiving member for use in electrophotography was prepared in the same manner as in Example 166 by further using  $\text{SiF}_4$  gas from a not illustrated cylinder in the lower layer and using  $\text{PH}_3/\text{H}_2$  gas in the upper layer, under the preparation conditions shown in Table 167 and, when evaluated in the same manner, satisfactory improvement was obtained to dots, coarse image and peeling in the same manner as in Example 166.

#### EXAMPLE 172

A light receiving member for use in electrophotography was prepared in the same manner as in Example 1 by using  $\text{PF}_5$  gas diluted with He gas (99.999% purity, hereinafter referred to as "PF<sub>5</sub>/He gas") and NO gas in the lower layer and, further using PF<sub>5</sub>/He, SiF<sub>4</sub> gas in the upper layer of Example 166, under the preparation conditions shown in Table 168 and, when evaluated in the same manner, satisfactory improvement was obtained to dots, coarse image and peeling in the same 50 manner as in Example 1.

#### EXAMPLE 173

A light receiving member for use in electrophotography was prepared in the same manner as in Example 166 by using  $\text{H}_2\text{S}$  gas (99.9% purity) in the lower layer and further using  $\text{PH}_3/\text{H}_2$  gas and  $\text{N}_2$  gas from not illustrated cylinder in the upper layer of Example 166, under the preparation conditions shown in Table 169 and, when evaluated in the same manner, satisfactory improvement was obtained to dots, coarse image and peeling in the same manner as in Example 166.

#### EXAMPLE 174

A light receiving member for use in electrophotography was prepared in the same manner as in Example 166 except for replacing  $\text{CH}_4$  gas cylinder with  $\text{C}_2\text{H}_2$  gas (99.9999% purity) cylinder and  $\text{PH}_3/\text{H}_2$  gas cylinder with  $\text{GeF}_4$  gas cylinder in Example 166, under the prep-

aration conditions shown in Table 170 and, when evaluated in the same manner, satisfactory improvement was obtained to the dots, coarse image and peeling in the same manner as in Example 166.

#### EXAMPLE 175

A light receiving member for use in electrophotography was prepared in the same manner as in Example 166, replacing  $B_2H_6$  gas cylinder with  $BF_3$  gas diluted with He gas (99.999% purity, hereinafter simply referred to as " $BF_3/He$ "), under the preparation conditions shown in Table 171 and, when evaluated in the same manner, satisfactory improvement was obtained to the dots, coarse image and peeling in the same manner as in Example 166.

#### EXAMPLE 176

A light receiving member for use in electrophotography was prepared in the same manner as in Example 166 by replacing NO gas cylinder with  $NH_3$  gas cylinder in Example 166, and further using  $SiF_4$  gas from not illustrated cylinder in Example 166, under the preparation conditions shown in Table 172 and, when evaluated in the same manner, satisfactory improvement was obtained to the dots, coarse image and peeling in the same manner as in Example 166.

#### EXAMPLE 177

A light receiving member for use in electrophotography was prepared in the same manner as in Example 171 by further using  $SiF_4$  gas from not illustrated cylinder in the upper layer of Example 171, under the preparation conditions shown in Table 174 and, when evaluated in the same manner, satisfactory improvement was obtained to dots, coarse image and peeling in the same manner as in Example 171.

#### EXAMPLE 178

A light receiving member for use in electrophotography was prepared in the same manner as in Example 174 by further using  $PH_3/H_2$  gas,  $Si_2F_6$  gas (99.99%, purity) and  $Si_2H_6$  gas (99.99% purity) from not illustrated cylinder, under the preparation conditions shown in Table 174 and, when evaluated in the same manner, satisfactory improvement was obtained to dots, coarse image and peeling in the same manner as in Example 174.

#### EXAMPLE 179

A light receiving member for use in electrophotography was prepared in the same manner as in Example 176 by replacing  $SiF_4$  gas with  $Si_2F_6$  gas and further using using  $B_2H_6/H_2$  gas in the lower layer, and further using  $PH_3/H_2$  gas in the upper layer, under the preparation conditions shown in Table 175 and, when evaluated in the same manner, satisfactory improvement was obtained to dots, coarse image and peeling in the same manner as in Example 176.

#### EXAMPLE 180

A light receiving member for use in electrophotography was prepared in the same manner as in Example 166 by further using  $PH_3H_2$  gas and  $GeH_4$  gas in the upper layer, under the preparation conditions shown in Table 176 and, when evaluated in the same manner, satisfactory improvement was obtained to dots, coarse image and peeling in the same manner as in Example 166.

#### EXAMPLE 181

A light receiving member for use in electrophotography was prepared in the same manner as in Example 166 by changing the outer diameter of the cylindrical aluminum support to 80 mm in Example 166, under the preparation conditions shown in Table 177 and, when evaluated in the same manner as in Example 1, except for using an electrophotographic apparatus, i.e., a copying machine NP-9030 manufactured by Canon Inc. and modified for the experimental use, satisfactory improvement was obtained to the dots, coarse image and peeling in the same manner as in Example 166.

#### EXAMPLE 182

A light receiving member for use in electrophotography was prepared in the same manner as in Example 166 by changing the outer diameter of the cylindrical aluminum support to 60 mm in Example 166, under the preparation conditions shown in Table 178 and, when evaluated in the same manner as in Example 166, except for using an electrophotographic apparatus, i.e., a copying machine NP-150Z manufactured by Canon Inc. and modified for the experimental use, satisfactory improvement was obtained to the dots, coarse image and peeling in the same manner as in Example 166.

#### EXAMPLE 183

A light receiving member for use in electrophotography was prepared in the same manner as in Example 166 by changing the outer diameter of the cylindrical aluminum support to 30 mm in Example 166, under the preparation conditions shown in Table 179 and, when evaluated in the same manner as in Example 166, except for using an electrophotographic apparatus, i.e., a copying machine FC-5 manufactured by Canon Inc. and modified for the experimental use, satisfactory improvement was obtained to the dots, coarse image and peeling in the same manner as in Example 166.

#### EXAMPLE 184

A light receiving member for use in electrophotography was prepared in the same manner as in Example 166 by changing the outer diameter of the cylindrical aluminum support to 15 mm in Example 166, under the preparation conditions shown in Table 180, and evaluated in the same manner as in Example 166, except for using an electrophotographic apparatus, manufactured for experimental use, satisfactory improvement was obtained to the dots, coarse image and peeling in the same manner as in Example 166.

#### EXAMPLE 185

A light sensitive member for use in electrophotography was prepared, under the same preparation conditions as those in Example 181 by using a cylindrical aluminum support applied with mirror-finishing fabrication in Example 181 and further machined into a cross sectional shape of :  $a=25$  um,  $b=0.8$  um as shown in FIG. 38 by a diamond point tool and, when evaluated in the same manner as in Example 181, satisfactory improvement was obtained to, the dots, coarse image and peeling in the same manner as in Example 181.

#### EXAMPLE 186

A light receiving member for use in electrophotography was prepared, under the same preparation conditions as those in Example 181 using a cylindrical alum-

num support applied with mirror-finish fabrication and subsequently applied with a so-called surface dimpling of causing a number of hit pits to the surface of the cylindrical aluminum support by the exposure to a plurality of dropping bearing balls to form into a cross sectional shape of:  $c=50$   $\mu\text{m}$  and  $d=1$   $\mu\text{m}$  as shown in FIG. 39 and, when evaluated in the same manner as in Example 181, satisfactory improvement was obtained for the dots, coarse image and peeling in the same manner as in Example 181.

#### EXAMPLE 187

A light receiving member for use in electrophotography having an upper layer comprising poly-Si(H, X) was prepared in the same manner as in Example 174 by using a cylindrical aluminum support heated to a temperature of 500° C., under the preparation conditions as shown in Table 181 and, when evaluated in the same manner, satisfactory improvement was obtained to dots, coarse image and peeling in the same manner as in Example 74.

#### EXAMPLE 188

A light receiving member for use in electrophotography was formed by microwave glow discharge decomposition in the same manner as in Example 23, further using SiF<sub>4</sub> gas, NO gas, Mg(C<sub>5</sub>H<sub>5</sub>)<sub>2</sub>/He gas and B<sub>2</sub>H<sub>6</sub> gas upon forming the lower layer in Example 23, under the preparing conditions shown in Table 182.

When the light receiving member for use in electrophotography was evaluated in the same manner in Example 166, improvement was obtained to the dots, coarse image and peeling in the same manner as in Example 166.

#### EXAMPLE 189

A light receiving member for use in electrophotography was prepared in the same manner as in Example 174, under the preparation conditions shown in Table 183 and, when evaluated in the same manner, satisfactory improvement was obtained to the dots, coarse image and peeling in the same manner as in Example 174.

#### EXAMPLE 190

A light receiving member for use in electrophotography was prepared in the same manner as in Example 175, under the preparation conditions shown in Table 184 and, when evaluated in the same manner, satisfactory improvement was obtained to the dots, coarse image and peeling in the same manner as in Example 175.

#### EXAMPLE 191

A light receiving member for use in electrophotography was prepared in the same manner as in Example 176, under the preparation conditions shown in Table 185 and, when evaluated in the same manner, satisfactory improvement was obtained to the dots, coarse image and peeling in the same manner as in Example 176.

#### EXAMPLE 192

A light receiving member for use in electrophotography was prepared in the same manner as in Example 177, under the preparation conditions shown in Table 186 and, when evaluated in the same manner, satisfactory improvement was obtained to the dots, coarse

image and peeling in the same manner as in Example 177.

#### EXAMPLE 193

A light receiving member for use in electrophotography was prepared in the same manner as in Example 178, under the preparation conditions shown in Table 187 and, when evaluated in the same manner, satisfactory improvement was obtained to the dots, coarse image and peeling in the same manner as in Example 178.

#### EXAMPLE 194

A light receiving member for use in electrophotography was prepared in the same manner as in Example 179, under the preparation conditions shown in Table 188 and, when evaluated in the same manner, satisfactory improvement was obtained to the dots, coarse image and peeling in the same manner as in Example 179.

#### EXAMPLE 195

A light receiving member for use in electrophotography was prepared in the same manner as in Example 169, under the preparation conditions shown in Table 189 and, when evaluated in the same manner, satisfactory improvement was obtained to the dots, coarse image and peeling in the same manner as in Example 169.

#### EXAMPLE 196

A light receiving member for use in electrophotography was prepared in the same manner as in Example 171, under the preparation conditions shown in Table 190 and, when evaluated in the same manner, satisfactory improvement was obtained to the dots, coarse image and peeling in the same manner as in Example 171.

#### EXAMPLE 197

A light receiving member for use in electrophotography was prepared in the same manner as in Example 177, under the preparation conditions shown in Table 191 and, when evaluated in the same manner, satisfactory improvement was obtained to the dots, coarse image and peeling in the same manner as in Example 177.

#### EXAMPLE 198

A light receiving member for use in electrophotography was prepared in the same manner as in Example 196, under the preparation conditions shown in Table 192 and, when evaluated in the same manner, satisfactory improvement was obtained to the dots, coarse image and peeling in the same manner as in Example 196.

#### EXAMPLE 199

A lower layer of a light receiving member for use in electrophotography according to this invention was formed by RF sputtering method and the upper layer thereof was formed by RF glow discharge decomposition.

FIG. 42 shows an apparatus for producing the light receiving member for use in electrophotography by the RF sputtering, comprising a raw material gas supply device 1500 and a deposition device 1501.

In the figure, a target 1045 is composed of Si, Al and Mg as the raw material for forming the lower layer, in which the mixing ratio for the atoms is varied such that a desired profile is obtained across the thickness for each of the atoms.

In the figure, raw material gases for forming the lower layer were tightly sealed in gas cylinders 1408, 1409 and 1410, in which the cylinder 1408 was for SiH<sub>4</sub> gas (99.99 % purity), the cylinder 1409 was for H<sub>2</sub> gas (99.9999 %) and the cylinder 1410 was for Ar gas (99.9999 % purity).

In the figure, a cylindrical aluminum support 1402 has an outer diameter of 108 mm and a mirror-finished surface.

At first, in the same manner as in Example 1, the inside of the deposition chamber 1401 and gas pipeways was evacuated till the pressure of the deposition chamber 1401 was reduced to  $1 \times 10^{-6}$  Torr.

Then, in the same manner as in Example 1, the respective gases were introduced into the mass flow controllers 1412 - 1414.

The temperature of the cylindrical aluminum support 1402 disposed in the deposition chamber 1401 was heated to 250° C. by a heater not illustrated.

After completing the preparation for the film formation as described above, the lower layer was formed on the cylindrical aluminum support 1402.

The lower layer was formed by gradually opening the flow-out valves 1420, 1421 and 1422, and the auxiliary valve 1432 thereby introducing the SiH<sub>4</sub> gas, H<sub>2</sub> gas and Ar gas to the inside of the deposition chamber 1401. In this case, the gas flow rates were controlled by the respective mass flow controllers 1412, 1413 and 1414 such that the gas flow rates were set to 20 SCCM for SiH<sub>4</sub>, 5 SCCM for H<sub>2</sub> gas, and 100 SCCM for Ar gas. The pressure in the deposition chamber 1401 was controlled to 0.01 Torr by adjusting the opening of the main valve 1407 while observing the vacuum meter 1435. Then, RF power was introduced between the target 1405 and the aluminum support 1402 by way of an RF matching box 1433 while setting the power of an RF power source (not illustrated) to 1 mW/cm<sup>3</sup>, thereby starting the formation of the lower layer on the cylindrical aluminum support. The mass flow controllers 1412, 1413 and 1414 were adjusted during formation of the lower layer such that the SiH<sub>4</sub> gas flow remained at a constant rate of 20 SCCM, the H<sub>2</sub> gas flow rate was increased at a constant ratio from 5 SCCM to 100 SCCM and the Ar gas flow rate remained at a constant ratio of 100 SCCM. Then, when the lower layer of 0.02 um thickness was formed, the RF glow discharge was stopped and the entrance of the gas to the inside of the deposition chamber 1401 was interrupted by closing the flow-out valves 1420, 1421 and 1423 and the auxiliary valve 1432, to complete the formation of the lower layer.

The cylindrical aluminum support 1402 was rotated at a desired speed by a driving device not illustrated during formation of the lower layer for making the layer formation uniform.

Then, a light receiving member for use in electrophotography was prepared in the same manner as in Example 166 under the preparation conditions shown in Table 193 by using the device illustrated in FIG. 37 upon forming the upper layer. When the same evaluation was applied, satisfactory improvement was obtained to dots, coarse image and layer peeling in the same manner as in Example 265.

## EXAMPLE 200

A light receiving member for use in electrophotography was prepared in the same manner as in Example 1 under the preparation conditions shown in Table 190 by further using Cu(C<sub>4</sub>H<sub>7</sub>N<sub>2</sub>O<sub>2</sub>)<sub>2</sub>/He gas upon forming the lower layer in Example 1.

## COMPARATIVE EXAMPLE 7

10 A light receiving member for use in electrophotography was prepared under the same preparation conditions as those in Example 1 except for not using H<sub>2</sub> gas and Cu(C<sub>4</sub>H<sub>7</sub>N<sub>2</sub>O<sub>2</sub>)<sub>2</sub>/He gas upon forming the lower layer. The conditions for preparing the light receiving member for use in electrophotography are shown in Table 195.

15 The light receiving members for use in electrophotography thus prepared in Example 200 and Comparative Example 7 were set respectively to an electrophotographic apparatus, i.e., a copying machine NP-7550 manufactured by Canon Inc. and modified for experimental use and, when several electrophotographic properties were checked under various conditions, it was found that both of them had outstanding characteristics in that they exhibit extremely good charging property.

20 Then, when the number of dots as the image characteristics were compared, it was found that the number of dots, particularly, the number of dots with less than 0.1 mm diameter of the light receiving member for use in electrophotography of Example 200 was less than  $\frac{1}{4}$  of that of the light receiving member for use in electrophotography in Comparative Example 7. In addition, for comparing the "coarse image", when the image 25 density was measured for circular regions each of 0.05 mm diameter assumed as one unit at 100 points and the scattering in the image density was evaluated, it was found that the scattering in the light receiving member for use in electrophotography of Example 200 was less than  $\frac{1}{5}$  for that of the light receiving member for use in electrophotography in Comparative Example 7 and the light receiving member for use in electrophotography of Example 200 was excellent over the light receiving member for use in Electrophotography of Comparative Example 7 in view of the visual observation.

30 In addition, for comparing the occurrence of image defects and the peeling of the light receiving layer due to impactive mechanical pressure applied for a relatively short period of time to the light receiving member for use in electrophotography, when stainless steel balls of 3.5 mm diameter were fallen freely from the vertical height of 30 cm above the surface of the light receiving member for use in electrophotography and abutted against the surface of the light receiving member for use in electrophotography, to thereby measure the frequency that cracks occurred to the light receiving layer, it was found that the rate of occurrence in the light receiving member for use in electrophotography of Example 200 was less than  $\frac{1}{5}$  for that in the light receiving member for use in electrophotography of Comparative Example 7.

35 When the lower layer of the light receiving member for use in electrophotography of Example 200 was analyzed by using SIMS, it was found that the content of silicon atoms, hydrogen atoms and aluminum atoms in the direction of the film thickness was varied as desired.

40 As has been described above, the light receiving member for use in electrophotography of Example 200

was superior to the light receiving member for use in electrophotography of Comparative Example 7.

#### EXAMPLE 201

A light receiving member for use in electrophotography was prepared in the same manner as in Example 200 by using  $B_2H_6/H_2$  gas and changing the way of varying the  $AlCl_3/He$  gas flow rate in the lower layer, under the preparation conditions shown in Table 196 and, when evaluated in the same manner, satisfactory improvement was obtained to the dots, coarse image and peeling in the same manner as in Example 200.

#### EXAMPLE 202

A light receiving member for use in electrophotography was prepared in the same manner as in Example 200 by using  $Mg(C_5H_5)_2$  gas diluted with He gas (hereinafter simply referred to as " $Mg(C_5H_5)_2/He$ ") from a not illustrated sealed vessel in the lower layer, and using He gas from a not illustrated cylinder and not using  $CH_4$  gas in the upper layer, under the preparation conditions shown in Table 197 and, when evaluated in the same manner, satisfactory improvement was obtained to the dots, coarse image and peeling in the same manner as in Example 292.

#### EXAMPLE 203

A light receiving member for use in electrophotography was prepared in the same manner as in Example 200 by further using  $Mg(C_5H_5)_2/He$  gas from a not illustrated sealed vessel,  $CH_4$  gas,  $B_2H_6/H_2$  gas,  $NO$  gas,  $SiF_4$  gas (99.999 % purity) from a not illustrated cylinder,  $N_2$  gas from a not illustrated cylinder and He gas, under the preparation conditions shown in Table 198 and, when evaluated in the same manner, satisfactory improvement was obtained to the dots, coarse image and peeling in the same manner as in Example 200.

#### EXAMPLE 204

A light receiving member for use in electrophotography was prepared in the same manner as in Example 200 by replacing  $H_2$  gas cylinder with  $Ar$  gas cylinder (99.9999 % purity),  $CH_4$  gas cylinder with  $NH_3$  gas cylinder (99.999 % purity), and further using  $SiF_4$  gas in the upper layer, under the preparation conditions shown in Table 199 and, when evaluated in the same manner, satisfactory improvement was obtained to the dots, coarse image and peeling in the same manner as in Example 200.

#### EXAMPLE 205

A light receiving member for use in electrophotography was prepared in the same manner as in Example 200 by further using  $CH_4$  gas and  $B_2H_6/H_2$  gas in the lower layer, and further using  $PH_3/H_2$  gas (99.999 % purity) from a not illustrated cylinder in the upper layer, under the preparation conditions shown in Table 200, and when evaluated in the same manner, satisfactory improvement was obtained to the dots, coarse image and peeling in the same manner as in Example 200.

#### EXAMPLE 206

A light receiving member for use in electrophotography was prepared in the same manner as in Example 200 by replacing  $NO$  gas cylinder with  $SiF_4$  gas cylinder in the lower layer, and further using  $Mg(C_5H_5)_2/He$  gas from a not illustrated sealed vessel in Example 200, and further using  $PF_5/H_2$  from not illustrated cylinder in

the upper layer, under the preparation conditions shown in Table 201 and, when evaluated in the same manner, satisfactory improvement was obtained to dots, coarse image and peeling in the same manner as in Example 200.

#### EXAMPLE 207

A light receiving member for use in electrophotography was prepared in the same manner as in Example 200 by using  $Mg(C_5H_5)_2/He$  gas from a not illustrated sealed vessel in the lower layer, and using  $PH_3/H_2$  gas from a not illustrated cylinder and  $N_2$  gas in the upper layer, under the preparation conditions shown in Table 202 and, when evaluated in the same manner, satisfactory improvement was obtained to dots, coarse image and peeling in the same manner as in Example 200.

#### EXAMPLE 208

A light receiving member for use in electrophotography was prepared in the same manner as in Example 200 by replacing  $CH_4$  gas cylinder with  $GeF_4$  gas (99.999 % purity) cylinder, further using  $CH_4$  gas and  $B_2H_6/H_2$  gas in the lower layer, and replacing  $CH_4$  gas cylinder with  $C_2H_2$  gas (99.9999 % purity) cylinder in the upper layer, under the preparation conditions shown in Table 203 and, when evaluated in the same manner, satisfactory improvement was obtained to dots, coarse image and peeling in the same manner as in Example 200.

#### EXAMPLE 209

A light receiving member for use in electrophotography was prepared in the same manner as in Example 200 by using  $Mg(C_5H_5)_2/He$  gas from a not illustrated sealed vessel, replacing  $B_2H_6$  gas cylinder with  $PH_3/H_2$  gas cylinder and further using  $SiF_4$  gas from a not illustrated cylinder, under the preparation conditions shown in Table 204 and, when evaluated in the same manner, satisfactory improvement was obtained to dots, coarse image and peeling in the same manner as in Example 204.

#### EXAMPLE 210

A light receiving member for use in electrophotography was prepared in the same manner as in Example 200 by replacing  $CH_4$  gas cylinder with  $NH_3$  gas (99.999 % purity) cylinder in Example 200, under the preparation conditions shown in Table 205 and, when evaluated in the same manner, satisfactory improvement was obtained to dots, coarse image and peeling in the same manner as in Example 200.

#### EXAMPLE 211

A light receiving member for use in electrophotography was prepared in the same manner as in Example 205 by further using  $CH_4$  gas and  $GeH_4$  gas in the lower layer, and further using  $SiF_4$  gas in the upper layer, under the preparation conditions shown in Table 206 and, when evaluated in the same manner, satisfactory improvement was obtained to the dots, coarse image and peeling in the same manner as in Example 205.

#### EXAMPLE 212

A light receiving member for use in electrophotography was prepared in the same manner as in Example 208 by replacing  $CH_4$  gas with  $C_2H_2$  gas, using  $PH_3/H_2$  gas from a not illustrated cylinder, and further using  $Si_2F_6$  gas (99.99 % purity) and  $Si_2F_6$  gas (99.99 a% purity) from not illustrated cylinders in the upper layer, under

the preparation conditions shown in Table 208 and, when evaluated in the same manner, satisfactory improvement was obtained to the dots, coarse image and peeling in the same manner as in Example 208.

#### EXAMPLE 213

A light receiving member for use in electrophotography was prepared in the same manner as in Example 200 by using  $\text{Si}_2\text{F}_6$  gas,  $\text{PH}_3$  gas and  $\text{NH}_3$  gas from not illustrated cylinders, under the preparation conditions shown in Table 208, and, when evaluated in the same manner, satisfactory improvement was obtained to the dots, coarse image and peeling in the same manner as in Example 200.

#### EXAMPLE 214

A light receiving member for use in electrophotography was prepared in the same manner as in Example 200 by further using  $\text{GeH}_4$  gas in the upper layer, under the preparation conditions shown in Table 209 and, when evaluated in the same manner, satisfactory improvement was obtained to the dots, coarse image and peeling in the same manner as in Example 200.

#### EXAMPLE 215

A light receiving member for use in electrophotography was prepared in the same manner as in Example 200 by changing the outer diameter of the cylindrical aluminum support to 80 mm in Example 200, under the preparation conditions shown in Table 210 and, when evaluated in the same manner as in Example 200, except for using an electrophotographic apparatus, i.e., a copying machine NP-9030 manufactured by Canon Inc. and modified for the experimental use, satisfactory improvement was obtained to the dots, coarse image and peeling in the same manner as in Example 200.

#### EXAMPLE 216

A light receiving member for use in electrophotography was prepared in the same manner as in Example 216 by changing the outer diameter of the cylindrical aluminum support to 60 mm in Example 216, under the preparation conditions shown in Table 211 and, when evaluated in the same manner as in Example 216, except for using an electrophotographic apparatus, i.e., a copying machine NP-150Z manufactured by Canon Inc. and modified for the experimental use, satisfactory improvement was obtained to the dots, coarse image and peeling in the same manner as in Example 216.

#### EXAMPLE 217

A light receiving member for use in electrophotography was prepared in the same manner as in Example 200 by changing the outer diameter of the cylindrical aluminum support to 30 mm in Example 200, under the preparation conditions shown in Table 212 and, when evaluated in the same manner as in Example 200, except for using an electrophotographic apparatus, i.e., a copying machine FC-5 manufactured by Canon Inc. and modified for the experimental use, satisfactory improvement was obtained to the dots, coarse image and peeling in the same manner as in Example 200.

#### EXAMPLE 218

A light receiving member for use in electrophotography was prepared in the same manner as in Example 200 by changing the outer diameter of the cylindrical aluminum support to 15 mm in Example 200, under the prepa-

ration conditions shown in Table 213, and evaluated in the same manner as in Example 200, except for using an electrophotographic apparatus, manufactured for experimental use and, when evaluated in the same manner, satisfactory improvement was obtained to the dots, coarse image and peeling in the same manner as in Example 200.

#### EXAMPLE 219

A light sensitive member for use in electrophotography was prepared, under the same preparation conditions as those in Example 215 by using a cylindrical aluminum support applied with mirror-finishing fabrication in Example 215 and further machined into a cross sectional shape of :  $a=25 \text{ um}$ ,  $b=0.8 \text{ um}$  as shown in FIG. 38 by a diamond point tool and, when evaluated in the same manner as in Example 215, satisfactory improvement was obtained to, the dots, coarse image and peeling in the same manner as in Example 215.

#### EXAMPLE 220

A light receiving member for use in electrophotography was prepared, under the same preparation conditions as those in Example 215 using a cylindrical aluminum support applied with mirror-finish fabrication and subsequently applied with a so-called surface dimpling of causing a number of hit pits to the surface of the cylindrical aluminum support by the exposure to a plurality of dropping bearing balls to form into a cross sectional shape of :  $c=50 \text{ um}$  and  $d=1 \text{ um}$  as shown in FIG. 39 and, when evaluated in the same manner as in Example 215, satisfactory improvement was obtained for the dots, coarse image and peeling in the same as in Example 215.

#### EXAMPLE 221

A light receiving member for use in electrophotography having an upper layer comprising poly- $\text{Si}(\text{H}, \text{X})$  was prepared in the same manner as in Example 208 by replacing  $\text{CH}_4$  gas with  $\text{C}_2\text{H}_2$  gas and using a cylindrical aluminum support heated to a temperature of  $500^\circ \text{ C.}$ , under the preparation conditions as shown in Table 214 and, when evaluated in the same manner, satisfactory improvement was obtained to dots, coarse image and peeling in the same manner as in Example 208.

#### EXAMPLE 222

A light receiving member for use in electrophotography was prepared by microwave glow discharge decomposition in the same manner as in Example 23 by further using  $\text{Cu}(\text{C}_4\text{H}_7\text{N}_2\text{O}_2)\text{He}$  gas,  $\text{SiF}_4$  gas,  $\text{NO}$  gas,  $\text{GeH}_4$  gas and  $\text{B}_2\text{H}_6$  gas upon forming the lower layer in Example 23, under the same preparation conditions as shown in Table 215.

When the light receiving member for use in electrophotography was evaluated in the same manner as in Example 200, satisfactory improvement was obtained to the dots, coarse image and peeling in the same manner as in Example 200.

When the lower layer of the light receiving member for use in electrophotography of Example 162 was analyzed by using SIMS, it was found that the content of silicon atoms, hydrogen atoms and aluminum atoms in the direction of the film thickness was varied as desired.

#### EXAMPLE 223

A light receiving member for use in electrophotography was prepared in the same manner as in Example 200

by replacing the  $\text{CH}_4$  gas cylinder with a  $\text{C}_2\text{H}_2$  gas cylinder in Example 200, under the preparation conditions shown in Table 216 and, when evaluated in the same manner, satisfactory improvement was obtained to the dots, coarse image and peeling in the same manner as in Example 200.

#### EXAMPLE 224

A light receiving member for use in electrophotography was prepared in the same manner as in Example 200 by replacing  $\text{B}_2\text{H}_6/\text{H}_2$  gas cylinder with  $\text{PF}_3/\text{H}_2$  gas cylinder in Example 200, further using  $\text{CH}_4$  gas in lower layer, and using  $\text{SiF}_4$  gas for the entire layer, under the preparation condition shown in Table 217 and, when evaluated in the same manner, satisfactory improvement was obtained to the dots, coarse image and peeling in the same manner as in Example 200.

#### EXAMPLE 225

A light receiving member for use in electrophotography was prepared in the same manner as in Example 200 by replacing  $\text{CH}_4$  gas cylinder with  $\text{NH}_3$  gas cylinder, using  $\text{SnH}_4$  from a not illustrated cylinder,  $\text{Mg}(\text{C}_5\text{H}_5)_2/\text{He}$  gas from a not illustrated sealed vessel in Example 200, under the preparation conditions shown in Table 218 and, when evaluated in the same manner, satisfactory improvement was obtained to the dots, coarse image and peeling in the same manner as in Example 200.

#### EXAMPLE 226

A light receiving member for use in electrophotography was prepared in the same manner as in Example 205 by replacing  $\text{B}_2\text{H}_6/\text{H}_2\text{N}_2$  gas cylinder with  $\text{PH}_3/\text{H}_2$  gas cylinder, and using  $\text{SiF}_4$  gas, under the preparation conditions shown in Table 219 and, when evaluated in the same manner, satisfactory improvement was obtained to the dots, coarse image and peeling in the same manner as in Example 205.

#### EXAMPLE 227

A light receiving member for use in electrophotography was prepared in the same manner as in Example 200 by replacing  $\text{CH}_4$  gas cylinder with  $\text{C}_2\text{H}_2$  gas cylinder, and further using  $\text{Si}_2\text{H}_6$  gas in the upper layer, under the preparation conditions shown in Table 220 and, when evaluated in the same manner, satisfactory improvement was obtained to the dots, coarse image and peeling in the same manner as in Example 200.

#### EXAMPLE 228

A light receiving member for use in electrophotography was prepared in the same manner as in Example 200 by replacing  $\text{CH}_4$  gas cylinder with  $\text{C}_2\text{H}_2$  gas cylinder, replacing  $\text{GeH}_4$  gas cylinder with  $\text{GeF}_4$  gas cylinder, and further using  $\text{PH}_3/\text{H}_2$  gas from a not illustrated gas cylinder in the upper layer, under the preparation conditions shown in Table 221 and, when evaluated in the same manner, satisfactory improvement was obtained to the dots, coarse image and peeling in the same manner as in Example 200.

#### EXAMPLE 229

A light receiving member for use in electrophotography was prepared, under the same manner as those in Example 200 using a cylindrical aluminum support applied with mirror-finish fabrication and subsequently applied with a so-called surface dimpling of causing a

number of hit pits to the surface of the cylindrical aluminum support by the exposure to a plurality of dropping bearing balls to form into a cross sectional shape of  $c=50 \mu\text{m}$  and  $d=1 \mu\text{m}$  as shown in FIG. 39 and, when evaluated in the same manner as in Example 200, satisfactory improvement was obtained for the dots, coarse image and peeling in the same as in Example 200.

#### EXAMPLE 230

A light receiving member for use in electrophotography was prepared in the same manner as in Example 200, under the preparation conditions shown in Table 223 and, when evaluated in the same manner, satisfactory improvement was obtained to the dots, coarse image and peeling in the same manner as in Example 200.

#### EXAMPLE 231

The lower layer was formed under the preparation conditions shown in Table 224 in the same manner as in Example 199 except for using a target composed of Si, Al, Cu instead of Si, Al, Mg used in forming the lower layer in Example 199.

Then, the upper layer was formed by glow discharge decomposition using the device shown in FIG. 37. Then, a light receiving member for use in electrophotography was prepared in the same manner as in Example 200 under the preparing conditions shown in a Table 224. When the evaluation was conducted in the same manner, satisfactory improvement to dots and layer peeling was obtained in the same manner as in Example 200.

When the lower layer of the light receiving member for use in electrophotography of Example 231 was analyzed by using SIMS, it was found that the content of silicon atoms, hydrogen atoms and aluminum atoms in the direction of the film thickness was varied as desired.

#### EXAMPLE 232

A light receiving member for use in electrophotography was prepared in the same manner as in Example 1 under the preparation conditions shown in Table 225 by further using  $\text{NaNH}_2/\text{He}$  gas upon forming the lower layer in Example 1.

#### COMPARATIVE EXAMPLE 8

A light receiving member for use in electrophotography was prepared under the same conditions in Example 232 except for not using  $\text{H}_2$  gas upon forming the lower layer.

The profile for the content of atoms across the layer thickness near the lower layer of the light receiving member for use in electrophotography in Example 232 and Comparative Example 8 thus prepared was analyzed by using SIMS (secondary ion mass analyzing device, manufactured by Kameka : IMS-3F). The results are shown in FIG. 43(a), (b). In FIG. 43, the abscissa represents the measured time corresponding to the position across the layer thickness, and the ordinate represents the content for each of the atoms by relative values.

FIG. 43(a) shows the profile for the content of atoms across the layer thickness in Example 232 in which aluminum atoms were distributed more on the side of the support, while silicon atoms and hydrogen atoms were distributed more on the side of the upper layer.

FIG. 43(b) shows the profile for the content of atoms across the layer thickness in Comparative Example 8 in

which aluminum atoms were distributed more on the side of the support, silicon atoms were distributed more on the side of the upper layer and hydrogen atoms were distributed uniformly.

Then, the light receiving members for use in electrophotography thus prepared in Example 232 and Comparative Example 8 were set respectively to electrophotographic apparatus, that is, a copying machine NP-7550 manufactured by Cannon Inc. and modified for experimental use and several electrophotographic properties were checked under various conditions.

The light receiving member for use in electrophotography was rotated for 1000 turns while using a magnet roller as a cleaning roller, coating positive toners on the magnet roller while keeping all of the charging devices not operated. Then, a black original was prepared by an ordinary electrophotographic process and, as a result of measuring the number of dots generated, it was found that the light receiving member for use in electrophotography of Example 232 showed the number of dots less than  $\frac{1}{3}$  for that of the light receiving member for use in electrophotography in Comparative Example 8.

In addition, the light receiving member for use in electrophotography was rotated by 20 turns in a state where coagulated paper dusts were placed on the grits of a separation charger to cause abnormal discharge. Then, after removing the paper dusts, images were prepared by using a black original and, as a result of measuring the number of dots, it was found that the number of dots in the light receiving member for use in electrophotography of Example 232 was less than  $\frac{1}{3}$  for that of the light receiving member for use in electrophotography in Comparative Example 8.

Further, a roll made of high density polyethylene having about 32 mm $\phi$  diameter and 5 mm thickness was urged to the light receiving member for use in electrophotography under the pressure of 2 kg and then the light receiving member for use in electrophotography was rotated for 500,000 turns. Then, as a result of comparing the number of peeling visually in the light receiving layer, it was found that the number of peeling for the light receiving member for use in Example 232 was less than  $\frac{1}{2}$  for that of the light receiving member for use in electrophotography in Comparative Example 8.

As has been described above, the light receiving member for use in electrophotography in Example 232 was superior from overall point of view to the light receiving member for use in electrophotography in Comparative Example 8.

#### EXAMPLE 233

A light receiving member for use in electrophotography was prepared in the same manner as in Example 232 under the preparing conditions shown in Table 226 except for changing the gas flow rate of  $\text{Al}(\text{CH}_3)_3/\text{He}$  to the value shown in Table 232.

#### COMPARATIVE EXAMPLE 9

A light receiving member for use in electrophotography was prepared in the same manner as in Example 232 under the preparing conditions shown in Table 225 except for changing the gas flow rate of  $\text{Al}(\text{CH}_3)_3/\text{He}$  to the value shown in Table 226.

A roll made of high density polyethylene was urged to the light receiving members for use in electrophotography thus prepared in Example 233, and Comparative Example 9 in the same manner as in Example 232 and the number of layer peeling was compared. The result is

shown in Table 226 assuming the number of layer peeling to 1 in the layer of the light receiving member for use in electrophotography of Example 232. Further, the content of aluminum atoms near the upper portion of the lower layer was analyzed by using SIMS. The result is shown in Table 226.

As shown by the result in Table 226, the number of layer peeling was low and satisfactory result was obtained in the region where the content of the aluminum atoms near the upper portion of the lower layer was greater than 20 atom%.

#### EXAMPLE 234

A light receiving member for use in electrophotography was prepared in the same manner as in Example 232 under the preparing conditions shown in Table 225 except for changing the temperature for the support at a constant rate from 350° C. to 250° C. and using  $\text{Y}(\text{O}-\text{C}_3\text{H}_7)_3$  instead of  $\text{NaNH}_2$  during formation of the lower layer. When the evaluation was conducted in the same manner, satisfactory improvement to dots and layer peeling was obtained in the same manner as in Example 232.

#### EXAMPLE 235

A light receiving member for use in electrophotography was prepared in the same manner as in Example 232 under the preparing conditions shown in Table 225 except for changing RF power at a constant rate from 50 mW/cm<sup>2</sup> to 5 mW/cm<sup>2</sup> and using  $\text{Mn}(\text{CH}_3)(\text{CO})_5$  instead of  $\text{NaNH}_2$  during formation of the lower layer. When the evaluation was conducted in the same manner, satisfactory improvement to dots and layer peeling was obtained in the same manner as in Example 232.

#### EXAMPLE 236

A light receiving member for use in electrophotography was prepared in the same manner as in Example 232 under the preparing conditions shown in Table 227 except for using  $\text{Zn}(\text{C}_2\text{H}_5)_2$  instead of  $\text{NaNH}_2$  and, further, adding the raw material gas shown in Table 227. When the evaluation was conducted in the same manner, satisfactory improvement to dots and layer peeling was obtained in the same manner as in Example 232.

#### EXAMPLE 237

A light receiving member for use in electrophotography was prepared in the same manner as in Example 232 under the preparing conditions shown in Table 225 except for changing the outer diameter of the cylindrical aluminum support to 30 mm and changing the gas flow rate and RF power shown in Table 225 to  $\frac{1}{3}$  respectively. When the evaluation was conducted in the same manner, satisfactory improvement to dots and layer peeling was obtained in the same manner as in Example 232.

#### EXAMPLE 238

A light receiving member for use in electrophotography was prepared in the same manner as in Example 232 under the preparing conditions shown in Table 228. When the evaluation was conducted in the same manner, satisfactory improvement to dots and layer peeling was obtained in the same manner as in Example 232.

#### EXAMPLE 239

A light receiving member for use in electrophotography was prepared by the microwave glow discharge

decomposition in the same manner as in Example 23 under the preparing conditions shown in Table 229 by further using SiF<sub>4</sub> gas and NaNH<sub>2</sub>/He gas upon forming the lower layer in Example 23.

When the same evaluation as in Example 232 was conducted for the light receiving member for use in electrophotography, satisfactory improvement was obtained to dots and layer peeling in the same manner as in Example 232.

The profile for the content of atoms across the layer thickness near the lower layer was analyzed by using SIMS in the same manner as in Example 232 and the result is shown in FIG. 43(c).

It was found that aluminum atoms, silicon atoms and hydrogen atoms are distributed in the same manner as in Example 232.

#### EXAMPLE 240

The lower layer was formed under the preparing conditions shown in Table 230 in the same manner as in Example 199 except for using a target composed of Si, Al, Mn instead of a target composed of Si, Al, Mg used upon forming the lower layer in Example 199.

Then, a light receiving member for use in electrophotography was prepared in the same manner as in Example 232 under the preparing conditions shown in Table 225 by using the device shown in FIG. 37 for forming

the same manner, satisfactory improvement to dots and layer peeling was obtained in the same manner as in Example 232.

The profile for the content of atoms across the layer thickness near the lower layer was analyzed by using SIMS in the manner as in Example 232 and the results is shown in FIG. 43(d).

It was found that aluminum atoms, silicon atoms and hydrogen atoms were distributed in the same manner as in Example 232.

In the following Tables 1 to 230, the mark “\*” means increase of a flow rate at constant proportion;

the mark “\*\*” means decrease of a flow rate at constant proportion;

the term “S-side” means substrate side;

the term “UL-side” means upper layer side;

the term “LL-side” means lower layer side;

the term “U.1st LR-side” means 1st layer region side

of the upper layer;

the term “U.2nd LR-side” means 2nd layer region side of the upper layer;

the term “U.3rd LR-side” means 3rd layer region side

of the upper layer;

the term “U.4th LR-side” means 4th layer region side

of the upper layer; and

the term “FS-side” means free surface side of the upper layer.

TABLE 1

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 50                          |                                            |                       |                      |
|                                  | H <sub>2</sub>                                            | 10→200*                     | 250                                        | 5                     | 0.4                  |
|                                  | AlCl <sub>3</sub> /He                                     | 120→40**                    |                                            |                       |                      |
|                                  | SiH <sub>4</sub>                                          | 100                         |                                            |                       |                      |
|                                  | B <sub>2</sub> H <sub>6</sub> (against SiH <sub>4</sub> ) | 200 ppm                     | 8                                          | 0.4                   | 3                    |
|                                  | H <sub>2</sub>                                            | 500                         |                                            |                       |                      |
| Upper layer                      | SiH <sub>4</sub>                                          | 300                         |                                            |                       |                      |
|                                  | H <sub>2</sub>                                            | 300                         | 250                                        | 15                    | 0.5                  |
|                                  | SiH <sub>4</sub>                                          | 50                          |                                            |                       |                      |
|                                  | CH <sub>4</sub>                                           | 500                         | 250                                        | 15                    | 0.4                  |
|                                  |                                                           |                             |                                            |                       | 0.5                  |

TABLE 2

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 50                          |                                            |                       |                      |
|                                  | AlCl <sub>3</sub> /He                                     | 120→40**                    | 250                                        | 5                     | 0.4                  |
|                                  | SiH <sub>4</sub>                                          | 100                         |                                            |                       |                      |
|                                  | B <sub>2</sub> H <sub>6</sub> (against SiH <sub>4</sub> ) | 200 ppm                     | 250                                        | 8                     | 0.4                  |
|                                  | H <sub>2</sub>                                            | 500                         |                                            |                       |                      |
|                                  | SiH <sub>4</sub>                                          | 300                         | 250                                        | 15                    | 0.5                  |
| Upper layer                      | SiH <sub>4</sub>                                          | 300                         |                                            |                       |                      |
|                                  | H <sub>2</sub>                                            | 300                         | 250                                        | 15                    | 0.5                  |
|                                  | SiH <sub>4</sub>                                          | 50                          |                                            |                       |                      |
|                                  | CH <sub>4</sub>                                           | 500                         | 250                                        | 10                    | 0.4                  |
|                                  |                                                           |                             |                                            |                       | 0.5                  |

the upper layer. When the evaluation was conducted in

TABLE 3

| Order of lamination (layer name) | Gases and their flow rates (SCCM)                                                | Substrate temperature (°C.) | RF discharging power (mW/cm <sup>3</sup> ) | Inner pressure (Torr) | Layer thickness (μm) |
|----------------------------------|----------------------------------------------------------------------------------|-----------------------------|--------------------------------------------|-----------------------|----------------------|
| Lower layer                      | SiH <sub>4</sub><br>H <sub>2</sub><br>AlCl <sub>3</sub> /He<br>(S-side: 0.01 μm) | 50<br>10→200*               | 250                                        | 5                     | 0.4                  |

TABLE 3-continued

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Upper layer region               | (UL-side: 0.01 μm)                                        | 10                          |                                            |                       |                      |
|                                  | SiH <sub>4</sub>                                          | 100                         |                                            |                       |                      |
|                                  | B <sub>2</sub> H <sub>6</sub> (against SiH <sub>4</sub> ) | 200 ppm                     | 250                                        | 8                     | 0.4                  |
|                                  | H <sub>2</sub>                                            | 500                         |                                            |                       |                      |
|                                  | SiH <sub>4</sub>                                          | 300                         |                                            |                       |                      |
|                                  | H <sub>2</sub>                                            | 300                         | 250                                        | 15                    | 0.5                  |
| 3rd layer region                 | SiH <sub>4</sub>                                          | 50                          |                                            |                       |                      |
|                                  | CH <sub>4</sub>                                           | 500                         | 250                                        | 10                    | 0.4                  |

TABLE 4

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 50                          |                                            |                       |                      |
|                                  | H <sub>2</sub>                                            | 5→200*                      | 150                                        | 0.5                   |                      |
|                                  | AlCl <sub>3</sub> /He (S-side: 0.01 μm)                   |                             | ↓                                          |                       |                      |
|                                  |                                                           | 300                         | 1.5                                        | 0.3                   | 0.02                 |
| Upper layer region               | (UL-side: 0.01 μm)                                        | 200→30**                    |                                            |                       |                      |
|                                  | SiH <sub>4</sub>                                          | 30→10**                     |                                            |                       |                      |
|                                  | H <sub>2</sub>                                            | 100                         |                                            |                       |                      |
|                                  | B <sub>2</sub> H <sub>6</sub> (against SiH <sub>4</sub> ) | 500 ppm                     | 250                                        | 10                    | 0.4                  |
|                                  | (LL-side: 2 μm)                                           |                             |                                            |                       |                      |
|                                  | (U·2nd·LR-side: 1 μm)                                     | 500 ppm→0**                 |                                            |                       |                      |
| 2nd layer region                 | H <sub>2</sub>                                            | 200                         |                                            |                       |                      |
|                                  | SiH <sub>4</sub>                                          | 300                         |                                            |                       |                      |
|                                  | H <sub>2</sub>                                            | 500                         | 250                                        | 20                    | 0.5                  |

TABLE 5

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 50                          |                                            |                       |                      |
|                                  | H <sub>2</sub>                                            | 5→200*                      |                                            |                       |                      |
|                                  | AlCl <sub>3</sub> /He (S-side: 0.01 μm)                   |                             | 250                                        | 1                     | 0.3                  |
|                                  | (UL-side: 0.01 μm)                                        | 200→30**                    |                                            |                       |                      |
| 1st layer region                 | SiH <sub>4</sub>                                          | 30→10**                     |                                            |                       |                      |
|                                  | H <sub>2</sub>                                            | 100                         |                                            |                       |                      |
|                                  | B <sub>2</sub> H <sub>6</sub> (against SiH <sub>4</sub> ) | 500 ppm                     |                                            |                       |                      |
|                                  | He                                                        | 600                         | 250                                        | 10                    | 0.4                  |
|                                  | AlCl <sub>3</sub> /He                                     | 0.1                         |                                            |                       |                      |
|                                  | SiF <sub>4</sub>                                          | 0.5                         |                                            |                       |                      |
| Upper layer                      | SiF <sub>4</sub>                                          |                             |                                            |                       |                      |
|                                  | NO                                                        | 0.1                         |                                            |                       |                      |
|                                  | CH <sub>4</sub>                                           | 1                           |                                            |                       |                      |
|                                  | 2nd layer region                                          | SiH <sub>4</sub>            | 300                                        |                       |                      |
|                                  | He                                                        | 600                         | 250                                        | 25                    | 0.6                  |
|                                  | B <sub>2</sub> H <sub>6</sub>                             | 0.3 ppm                     |                                            |                       |                      |
| 3rd layer region                 | SiF <sub>4</sub>                                          | 0.5                         |                                            |                       |                      |
|                                  | AlCl <sub>3</sub> /He                                     | 0.1                         |                                            |                       |                      |
|                                  | SiH <sub>4</sub>                                          | 50                          |                                            |                       |                      |
|                                  | CH <sub>4</sub>                                           | 500                         |                                            |                       |                      |
|                                  | NO                                                        | 0.1                         | 250                                        | 10                    | 0.4                  |
|                                  | B <sub>2</sub> H <sub>6</sub>                             | 0.3 ppm                     |                                            |                       |                      |

TABLE 6

| Order of lamination (layer name) | Gases and their flow rates (SCCM)       | Substrate temperature (°C.) | RF discharging power (mW/cm <sup>3</sup> ) | Inner pressure (Torr) | Layer thickness (μm) |
|----------------------------------|-----------------------------------------|-----------------------------|--------------------------------------------|-----------------------|----------------------|
| Lower layer                      | SiH <sub>4</sub>                        | 10→100*                     |                                            |                       |                      |
|                                  | H <sub>2</sub>                          | 5→200*                      |                                            |                       |                      |
|                                  | AlCl <sub>3</sub> /He (S-side: 0.05 μm) |                             | 250                                        | 10                    | 0.4                  |
|                                  |                                         | 200→40**                    |                                            |                       | 0.2                  |

TABLE 6-continued

| Order of lamination (layer name) | Gases and their flow rates (SCCM)                                                                         | Substrate temperature (°C.) | RF discharging power (mW/cm <sup>3</sup> ) | Inner pressure (Torr) | Layer thickness (μm) |
|----------------------------------|-----------------------------------------------------------------------------------------------------------|-----------------------------|--------------------------------------------|-----------------------|----------------------|
|                                  | (UL-side: 0.15 μm)                                                                                        |                             |                                            |                       |                      |
| Upper layer                      | SiH <sub>4</sub>                                                                                          | 40→10**                     |                                            |                       |                      |
| 1st layer region                 | B <sub>2</sub> H <sub>6</sub> (against SiH <sub>4</sub> )<br>(LL-side: 2 μm)<br>(U · 2nd · LR-side: 1 μm) | 100<br>500 ppm              | 250                                        | 10                    | 0.4                  |
| 2nd layer region                 | H <sub>2</sub><br>SiH <sub>4</sub><br>Ar                                                                  | 200<br>400<br>200           | 250                                        | 10                    | 0.5                  |
| 3rd layer region                 | SiH <sub>4</sub><br>NH <sub>3</sub>                                                                       | 100<br>30                   | 250                                        | 5                     | 0.4                  |
|                                  |                                                                                                           |                             |                                            |                       | 0.3                  |

TABLE 7

| Order of lamination (layer name) | Gases and their flow rates (SCCM)                                                                                                                                                                                                      | Substrate temperature (°C.)                                                                              | RF discharging power (mW/cm <sup>3</sup> ) | Inner pressure (Torr)           | Layer thickness (μm)         |
|----------------------------------|----------------------------------------------------------------------------------------------------------------------------------------------------------------------------------------------------------------------------------------|----------------------------------------------------------------------------------------------------------|--------------------------------------------|---------------------------------|------------------------------|
| Lower layer                      | SiH <sub>4</sub><br>H <sub>2</sub><br>AlCl <sub>3</sub> /He<br>(S-side: 0.05 μm)                                                                                                                                                       | 10→100*<br>5→200*                                                                                        | 300                                        | 10                              | 0.4                          |
| Upper layer                      | SiH <sub>4</sub><br>B <sub>2</sub> H <sub>6</sub><br>H <sub>2</sub><br>SiH <sub>4</sub><br>H <sub>2</sub><br>SiH <sub>4</sub><br>CH <sub>4</sub><br>PH <sub>3</sub> (against SiH <sub>4</sub> )<br>SiH <sub>4</sub><br>CH <sub>4</sub> | 200→40**<br>40→10**<br>100<br>200 ppm<br>500<br>300<br>500<br>600<br>3000 ppm<br>100<br>600<br>40<br>300 | 8<br>20<br>300<br>300<br>300<br>15<br>10   | 0.4<br>0.5<br>0.5<br>0.4<br>0.4 | 0.2<br>0.5<br>20<br>7<br>0.1 |

TABLE 8

| Order of lamination (layer name) | Gases and their flow rates (SCCM)                                                                                                                                                                                                                                                                                             | Substrate temperature (°C.)                                                                  | RF discharging power (mW/cm <sup>3</sup> )         | Inner pressure (Torr)              | Layer thickness (μm) |
|----------------------------------|-------------------------------------------------------------------------------------------------------------------------------------------------------------------------------------------------------------------------------------------------------------------------------------------------------------------------------|----------------------------------------------------------------------------------------------|----------------------------------------------------|------------------------------------|----------------------|
| Lower layer                      | SiH <sub>4</sub><br>H <sub>2</sub><br>AlCl <sub>3</sub> /He                                                                                                                                                                                                                                                                   | 50<br>5→200*<br>200→20**                                                                     | 330                                                | 5                                  | 0.4                  |
| Upper layer                      | SiH <sub>4</sub><br>PH <sub>3</sub><br>H <sub>2</sub><br>SiH <sub>4</sub><br>SiF <sub>4</sub><br>H <sub>2</sub><br>SiH <sub>4</sub><br>CH <sub>4</sub><br>B <sub>2</sub> H <sub>6</sub><br>(against SiH <sub>4</sub> )<br>SiH <sub>4</sub><br>CH <sub>4</sub><br>B <sub>2</sub> H <sub>6</sub><br>(against SiH <sub>4</sub> ) | 100<br>100 ppm<br>100<br>400<br>10<br>800<br>100<br>400<br>5000 ppm<br>20<br>400<br>8000 ppm | 330<br>330<br>330<br>330<br>25<br>350<br>350<br>10 | 8<br>25<br>0.5<br>15<br>0.4<br>0.4 | 3<br>25<br>5<br>1    |

TABLE 9

| Order of lamination (layer name) | Gases and their flow rates (SCCM)                                                | Substrate temperature (°C.) | RF discharging power (mW/cm <sup>3</sup> ) | Inner pressure (Torr) | Layer thickness (μm) |
|----------------------------------|----------------------------------------------------------------------------------|-----------------------------|--------------------------------------------|-----------------------|----------------------|
| Lower layer                      | SiH <sub>4</sub><br>H <sub>2</sub><br>AlCl <sub>3</sub> /He<br>(S-side: 0.01 μm) | 50<br>5→200*                | 300                                        | 1                     | 0.3                  |
|                                  | 200→30**<br>(UL-side: 0.01 μm)                                                   |                             |                                            |                       |                      |

TABLE 9-continued

| Order of lamination (layer name) | Gases and their flow rates (SCCM) |                                                           | Substrate temperature (°C.) | RF discharging power (mW/cm <sup>3</sup> ) | Inner pressure (Torr) | Layer thickness (μm) |
|----------------------------------|-----------------------------------|-----------------------------------------------------------|-----------------------------|--------------------------------------------|-----------------------|----------------------|
| Upper layer                      | 1st layer region                  | SiH <sub>4</sub>                                          | 30→10**                     |                                            |                       |                      |
|                                  | 1st layer region                  | B <sub>2</sub> H <sub>6</sub> (against SiH <sub>4</sub> ) | 100                         |                                            |                       |                      |
|                                  | 2nd layer region                  | H <sub>2</sub>                                            | 200 ppm                     | 300                                        | 8                     | 0.4                  |
|                                  | 2nd layer region                  | H <sub>2</sub>                                            | 500                         |                                            |                       |                      |
|                                  | 3rd layer region                  | SiH <sub>4</sub>                                          | 300                         |                                            |                       |                      |
|                                  | 4th layer region                  | N <sub>2</sub>                                            | 200                         | 300                                        | 20                    | 0.5                  |
| Lower layer                      | 3rd layer region                  | PH <sub>3</sub> (against SiH <sub>4</sub> )               | 50                          |                                            |                       |                      |
|                                  | 4th layer region                  | SiH <sub>4</sub>                                          | 500                         | 3000 ppm                                   |                       |                      |
| Lower layer                      | 4th layer region                  | CH <sub>4</sub>                                           | 40                          |                                            |                       |                      |
|                                  | Lower layer                       | CH <sub>4</sub>                                           | 600                         | 300                                        | 10                    | 0.3                  |

TABLE 10

| Order of lamination (layer name) | Gases and their flow rates (SCCM) |                                                           | Substrate temperature (°C.) | RF discharging power (mW/cm <sup>3</sup> ) | Inner pressure (Torr) | Layer thickness (μm) |
|----------------------------------|-----------------------------------|-----------------------------------------------------------|-----------------------------|--------------------------------------------|-----------------------|----------------------|
| Upper layer                      | 1st layer region                  | SiH <sub>4</sub>                                          | 50                          |                                            |                       |                      |
|                                  | 1st layer region                  | H <sub>2</sub>                                            | 5→200*                      | 250                                        | 5                     | 0.4                  |
|                                  | 1st layer region                  | AlCl <sub>3</sub> /He                                     | 200→20**                    |                                            |                       |                      |
|                                  | 1st layer region                  | SiH <sub>4</sub>                                          | 100                         |                                            |                       |                      |
|                                  | 2nd layer region                  | B <sub>2</sub> H <sub>6</sub> (against SiH <sub>4</sub> ) | 500 ppm                     |                                            |                       |                      |
|                                  | 2nd layer region                  | (LL-side: 3 μm)<br>(U·2nd·LR-side: 2 μm)                  | 50<br>500 ppm→0**           | 10                                         | 0.4                   | 5                    |
| Lower layer                      | 3rd layer region                  | H <sub>2</sub>                                            | 200                         |                                            |                       |                      |
|                                  | 3rd layer region                  | AlCl <sub>3</sub> /He (against SiH <sub>4</sub> )         | 1→0**                       |                                            |                       |                      |
|                                  | 4th layer region                  | SiH <sub>4</sub>                                          | 300                         |                                            |                       |                      |
|                                  | 4th layer region                  | H <sub>2</sub>                                            | 300                         | 250                                        | 15                    | 0.5                  |
|                                  | 4th layer region                  | SiH <sub>4</sub>                                          | 200                         |                                            |                       |                      |
|                                  | 4th layer region                  | C <sub>2</sub> H <sub>2</sub>                             | 10→20*                      | 250                                        | 15                    | 0.4                  |
| Lower layer                      | 4th layer region                  | NO                                                        | 1                           |                                            |                       | 20                   |

TABLE 11

| Order of lamination (layer name) | Gases and their flow rates (SCCM) |                                                           | Substrate temperature (°C.) | RF discharging power (mW/cm <sup>3</sup> ) | Inner pressure (Torr) | Layer thickness (μm) |
|----------------------------------|-----------------------------------|-----------------------------------------------------------|-----------------------------|--------------------------------------------|-----------------------|----------------------|
| Upper layer                      | 1st layer region                  | SiH <sub>4</sub>                                          | 50                          |                                            |                       |                      |
|                                  | 1st layer region                  | H <sub>2</sub>                                            | 5→200*                      | 250                                        | 1                     | 0.4                  |
|                                  | 1st layer region                  | AlCl <sub>3</sub> /He (S-side: 0.01 μm)                   | 200→30**                    |                                            |                       |                      |
|                                  | 1st layer region                  | (UL-side: 0.01 μm)                                        | 30→10**                     |                                            |                       |                      |
|                                  | 2nd layer region                  | SiH <sub>4</sub>                                          | 100                         |                                            |                       |                      |
|                                  | 2nd layer region                  | B <sub>2</sub> H <sub>6</sub> (against SiH <sub>4</sub> ) | 500 ppm                     | 250                                        | 10                    | 0.4                  |
| Lower layer                      | 2nd layer region                  | (LL-side: 2 μm)<br>(U·2nd·LR-side: 1 μm)                  | 500 ppm→0**                 |                                            |                       |                      |
|                                  | 3rd layer region                  | H <sub>2</sub>                                            | 200                         |                                            |                       |                      |
|                                  | 3rd layer region                  | SiH <sub>4</sub>                                          | 300                         | 300                                        | 20                    | 0.5                  |
|                                  | 3rd layer region                  | H <sub>2</sub>                                            | 300                         |                                            |                       |                      |
|                                  | 4th layer region                  | SiH <sub>4</sub>                                          | 100                         | 300                                        | 15                    | 0.4                  |
|                                  | 4th layer region                  | CH <sub>4</sub>                                           | 100                         |                                            |                       |                      |
| Lower layer                      | 4th layer region                  | SiH <sub>4</sub>                                          | 50                          | 300                                        | 10                    | 0.4                  |
|                                  | 4th layer region                  | CH <sub>4</sub>                                           | 600                         |                                            |                       | 0.5                  |

TABLE 12

| Order of lamination (layer name) | Gases and their flow rates (SCCM)       |         | Substrate temperature (°C.) | RF discharging power (mW/cm <sup>3</sup> ) | Inner pressure (Torr) | Layer thickness (μm) |
|----------------------------------|-----------------------------------------|---------|-----------------------------|--------------------------------------------|-----------------------|----------------------|
| Lower layer                      | SiH <sub>4</sub>                        | 10→100* |                             |                                            |                       |                      |
| Lower layer                      | H <sub>2</sub>                          | 5→200*  | 300                         | 5                                          | 0.4                   | 0.2                  |
| Lower layer                      | AlCl <sub>3</sub> /He (S-side: 0.05 μm) |         |                             |                                            |                       |                      |

TABLE 12-continued

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Upper layer                      | 200→40**<br>(UL-side: 0.15 μm)                            |                             |                                            |                       |                      |
|                                  | 40→10**                                                   |                             |                                            |                       |                      |
|                                  | 1st layer region SiH <sub>4</sub>                         | 100                         |                                            |                       |                      |
|                                  | B <sub>2</sub> H <sub>6</sub> (against SiH <sub>4</sub> ) | 200 ppm                     | 300                                        | 5                     | 0.4                  |
|                                  | H <sub>2</sub>                                            | 500                         |                                            |                       |                      |
|                                  | 2nd layer region SiH <sub>4</sub>                         | 100                         |                                            |                       |                      |
|                                  | H <sub>2</sub>                                            | 300                         | 300                                        | 5                     | 0.2                  |
|                                  | 3rd layer region SiH <sub>4</sub>                         | 300                         |                                            | 15                    | 0.4                  |
|                                  | NH <sub>3</sub>                                           | 50                          | 300                                        |                       | 25                   |
|                                  | 4th layer region SiH <sub>4</sub>                         | 100                         |                                            | 10                    | 0.4                  |
|                                  | NH <sub>3</sub>                                           | 50                          | 300                                        |                       | 0.3                  |

TABLE 13

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Upper layer                      | SiH <sub>4</sub>                                          | 10→100*                     |                                            |                       |                      |
|                                  | H <sub>2</sub>                                            | 5→200*                      |                                            |                       |                      |
|                                  | AlCl <sub>3</sub> /He                                     | 250                         | 5                                          | 0.4                   | 0.2                  |
|                                  | (S-side: 0.05 μm)                                         |                             |                                            |                       |                      |
|                                  | 200→40**<br>(UL-side: 0.15 μm)                            |                             |                                            |                       |                      |
|                                  | 40→10**                                                   |                             |                                            |                       |                      |
|                                  | 1st layer region SiH <sub>4</sub>                         | 100                         |                                            |                       |                      |
|                                  | B <sub>2</sub> H <sub>6</sub> (against SiH <sub>4</sub> ) | 500 ppm                     | 250                                        | 8                     | 0.4                  |
|                                  | (LL-side: 2 μm)                                           |                             |                                            |                       |                      |
|                                  | (U·2nd·LR-side: 1 μm)                                     |                             |                                            |                       |                      |
|                                  | 500 ppm→0**                                               |                             |                                            |                       |                      |
|                                  | 2nd layer region H <sub>2</sub>                           | 200                         |                                            |                       |                      |
|                                  | SiH <sub>4</sub>                                          | 100                         |                                            |                       |                      |
|                                  | SiF <sub>4</sub>                                          | 5                           | 300                                        | 3                     | 0.5                  |
|                                  | H <sub>2</sub>                                            | 200                         |                                            |                       |                      |
|                                  | 3rd layer region SiH <sub>4</sub>                         | 100                         |                                            |                       |                      |
|                                  | CH <sub>4</sub>                                           | 100                         | 300                                        | 15                    | 0.4                  |
|                                  | PH <sub>3</sub> (against SiH <sub>4</sub> )               | 50 ppm                      |                                            |                       | 30                   |
|                                  | 4th layer region SiH <sub>4</sub>                         | 50                          |                                            |                       |                      |
|                                  | CH <sub>4</sub>                                           | 600                         | 300                                        | 10                    | 0.4                  |
|                                  |                                                           |                             |                                            |                       | 0.5                  |

TABLE 14

| Order of lamination (layer name) | Gases and their flow rates (SCCM)                            | Substrate temperature (°C.) | RF discharging power (mW/cm <sup>3</sup> ) | Inner pressure (Torr) | Layer thickness (μm) |
|----------------------------------|--------------------------------------------------------------|-----------------------------|--------------------------------------------|-----------------------|----------------------|
| Upper layer                      | SiH <sub>4</sub>                                             | 50                          |                                            |                       |                      |
|                                  | H <sub>2</sub>                                               | 5→200*                      | 250                                        | 5                     | 0.4                  |
|                                  | AlCl <sub>3</sub> /He                                        | 200→20**                    |                                            |                       |                      |
|                                  | SiH <sub>4</sub>                                             | 40                          |                                            |                       |                      |
|                                  | 1st layer region PH <sub>3</sub> (against SiH <sub>4</sub> ) | 250 ppm                     | 250                                        | 8                     | 0.4                  |
|                                  | (LL-side: 1 μm)                                              |                             |                                            |                       |                      |
|                                  | (U·2nd·LR-side: 1 μm)                                        |                             |                                            |                       |                      |
|                                  | 250 ppm→0**                                                  |                             |                                            |                       |                      |
|                                  | 2nd layer region H <sub>2</sub>                              | 40                          |                                            |                       |                      |
|                                  | Si <sub>2</sub> H <sub>6</sub>                               | 200                         |                                            |                       |                      |
|                                  | H <sub>2</sub>                                               | 200                         | 300                                        | 10                    | 0.5                  |
|                                  | 3rd layer region SiH <sub>4</sub>                            | 300                         |                                            |                       |                      |
|                                  | C <sub>2</sub> H <sub>2</sub>                                | 50                          | 330                                        | 20                    | 0.4                  |
|                                  | B <sub>2</sub> H <sub>6</sub> (against SiH <sub>4</sub> )    |                             |                                            |                       | 30                   |
|                                  | (U·2nd·LR-side: 1 μm)                                        |                             |                                            |                       |                      |
|                                  | 1→100 ppm*                                                   |                             |                                            |                       |                      |
|                                  | (U·4th·LR-side: 29 μm)                                       |                             |                                            |                       |                      |
|                                  | 100 ppm                                                      |                             |                                            |                       |                      |
|                                  | 4th layer region SiH <sub>4</sub>                            | 200                         | 330                                        | 10                    | 0.4                  |
|                                  | C <sub>2</sub> H <sub>2</sub>                                | 200                         |                                            |                       | 1                    |

TABLE 15

| Order of lamination (layer name) | Gases and their flow rates (SCCM)                                            | Substrate temperature (°C.) | RF discharging power (mW/cm <sup>3</sup> ) | Inner pressure (Torr) | Layer thickness (μm) |
|----------------------------------|------------------------------------------------------------------------------|-----------------------------|--------------------------------------------|-----------------------|----------------------|
| Lower layer                      | SiH <sub>4</sub> 10→100*                                                     | 250                         | 5                                          | 0.4                   | 0.2                  |
|                                  | H <sub>2</sub> 5→200*                                                        |                             |                                            |                       |                      |
|                                  | AlCl <sub>3</sub> /He (S-side: 0.05 μm)                                      |                             |                                            |                       |                      |
|                                  | (UL-side: 0.15 μm) 200→40**                                                  |                             |                                            |                       |                      |
| Upper layer                      | 1st layer SiH <sub>4</sub> 100                                               | 300                         | 8                                          | 0.3                   | 3                    |
|                                  | 2nd region B <sub>2</sub> H <sub>6</sub> (against SiH <sub>4</sub> ) 200 ppm |                             |                                            |                       |                      |
|                                  | 2nd layer H <sub>2</sub> 500                                                 | 300                         | 5                                          | 0.2                   | 8                    |
|                                  | 3rd region SiH <sub>4</sub> 100                                              |                             |                                            |                       |                      |
|                                  | 3rd layer H <sub>2</sub> 300                                                 | 300                         | 15                                         | 0.4                   | 25                   |
|                                  | 4th region PH <sub>3</sub> (against SiH <sub>4</sub> ) 50 ppm                |                             |                                            |                       |                      |
|                                  | 4th layer NH <sub>3</sub> 100                                                | 300                         | 5                                          | 0.4                   | 0.7                  |
|                                  | region PH <sub>3</sub> (against SiH <sub>4</sub> ) 80→100*                   |                             |                                            |                       |                      |
|                                  | region NH <sub>3</sub> 500 ppm                                               |                             |                                            |                       |                      |

TABLE 16

| Order of lamination (layer name) | Gases and their flow rates (SCCM)       | Substrate temperature (°C.) | RF discharging power (mW/cm <sup>3</sup> ) | Inner pressure (Torr) | Layer thickness (μm) |
|----------------------------------|-----------------------------------------|-----------------------------|--------------------------------------------|-----------------------|----------------------|
| Lower layer                      | SiH <sub>4</sub> 50                     | 250                         | 1                                          | 0.4                   | 0.02                 |
|                                  | H <sub>2</sub> 5→200*                   |                             |                                            |                       |                      |
|                                  | AlCl <sub>3</sub> /He (S-side: 0.01 μm) |                             |                                            |                       |                      |
|                                  | (UL-side: 0.01 μm) 200→30**             |                             |                                            |                       |                      |
| Upper layer                      | 1st layer SiH <sub>4</sub> 100          | 300                         | 8                                          | 0.4                   | 3                    |
|                                  | 2nd region PH <sub>3</sub> 100 ppm      |                             |                                            |                       |                      |
|                                  | 2nd layer H <sub>2</sub> 100            | 300                         | 20                                         | 0.5                   | 20                   |
|                                  | 3rd region SiH <sub>4</sub> 300         |                             |                                            |                       |                      |
|                                  | 3rd layer H <sub>2</sub> 500            | 300                         | 5                                          | 0.4                   | 1                    |
|                                  | 4th region GeH <sub>4</sub> 10→50*      |                             |                                            |                       |                      |
|                                  | 4th layer H <sub>2</sub> 300            | 300                         | 10                                         | 0.4                   | 1                    |
|                                  | region SiH <sub>4</sub> 100→40**        |                             |                                            |                       |                      |
|                                  | region CH <sub>4</sub> 100→600*         |                             |                                            |                       |                      |

TABLE 17

| Order of lamination (layer name) | Gases and their flow rates (SCCM)                                            | Substrate temperature (°C.) | RF discharging power (mW/cm <sup>3</sup> ) | Inner pressure (Torr) | Layer thickness (μm) |
|----------------------------------|------------------------------------------------------------------------------|-----------------------------|--------------------------------------------|-----------------------|----------------------|
| Lower layer                      | SiH <sub>4</sub> 50                                                          | 300                         | 1                                          | 0.3                   | 0.02                 |
|                                  | H <sub>2</sub> 5→200*                                                        |                             |                                            |                       |                      |
|                                  | AlCl <sub>3</sub> /He (S-side: 0.01 μm)                                      |                             |                                            |                       |                      |
|                                  | (UL-side: 0.01 μm) 200→30**                                                  |                             |                                            |                       |                      |
| Upper layer                      | 1st layer SiH <sub>4</sub> 100                                               | 300                         | 8                                          | 0.4                   | 10                   |
|                                  | 2nd region B <sub>2</sub> H <sub>6</sub> (against SiH <sub>4</sub> ) 200 ppm |                             |                                            |                       |                      |
|                                  | 2nd layer SiH <sub>4</sub> 300                                               | 300                         | 15                                         | 0.5                   | 20                   |
|                                  | 3rd region H <sub>2</sub> 400                                                |                             |                                            |                       |                      |
|                                  | 3rd layer CH <sub>4</sub> 50                                                 | 300                         | 10                                         | 0.4                   | 0.5                  |
|                                  | region CH <sub>4</sub> 500                                                   |                             |                                            |                       |                      |
|                                  |                                                                              |                             |                                            |                       |                      |

TABLE 18

| Order of lamination (layer name) | Gases and their flow rates (SCCM) | Substrate temperature (°C.) | RF discharging power (mW/cm <sup>3</sup> ) | Inner pressure (Torr) | Layer thickness (μm) |
|----------------------------------|-----------------------------------|-----------------------------|--------------------------------------------|-----------------------|----------------------|
|                                  | SiH <sub>4</sub> 50               |                             |                                            |                       |                      |
|                                  | H <sub>2</sub> 5→200*             |                             |                                            |                       |                      |

TABLE 18-continued

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | AlCl <sub>3</sub> /He (S-side: 0.01 μm)                           | 300                         | 0.7                                        | 0.3                   | 0.02                 |
|                                  | 200→30** (UL-side: 0.01 μm)                                       |                             |                                            |                       |                      |
|                                  | 30→10**                                                           |                             |                                            |                       |                      |
| 1st layer                        | SiH <sub>4</sub> 80                                               |                             |                                            |                       |                      |
| Upper layer                      | H <sub>2</sub> 400                                                | 300                         | 7                                          | 0.3                   | 10                   |
| 2nd layer region                 | B <sub>2</sub> H <sub>6</sub> (against SiH <sub>4</sub> ) 200 ppm |                             |                                            |                       |                      |
| 3rd layer region                 | SiH <sub>4</sub> 200                                              |                             |                                            |                       |                      |
|                                  | H <sub>2</sub> 400                                                | 300                         | 12                                         | 0.4                   | 20                   |
|                                  | SiH <sub>4</sub> 40                                               |                             |                                            |                       |                      |
|                                  | CH <sub>4</sub> 400                                               | 300                         | 7                                          | 0.3                   | 0.5                  |

TABLE 19

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 25                                               |                             |                                            |                       |                      |
|                                  | H <sub>2</sub> 5→100*                                             | 300                         | 0.5                                        | 0.2                   | 0.02                 |
|                                  | AlCl <sub>3</sub> /He (S-side: 0.01 μm)                           |                             |                                            |                       |                      |
|                                  | 100→15** (UL-side: 0.01 μm)                                       |                             |                                            |                       |                      |
|                                  | 15→5**                                                            |                             |                                            |                       |                      |
| Upper layer                      | SiH <sub>4</sub> 60                                               |                             |                                            |                       |                      |
| 1st layer region                 | H <sub>2</sub> 300                                                | 300                         | 6                                          | 0.2                   | 10                   |
|                                  | B <sub>2</sub> H <sub>6</sub> (against SiH <sub>4</sub> ) 200 ppm |                             |                                            |                       |                      |
| 2nd layer region                 | SiH <sub>4</sub> 150                                              |                             |                                            |                       |                      |
|                                  | H <sub>2</sub> 300                                                | 300                         | 10                                         | 0.4                   | 20                   |
| 3rd layer region                 | SiH <sub>4</sub> 30                                               |                             |                                            |                       |                      |
|                                  | CH <sub>4</sub> 300                                               | 300                         | 5                                          | 0.3                   | 0.5                  |

TABLE 20

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 20                                               |                             |                                            |                       |                      |
|                                  | H <sub>2</sub> 5→100*                                             | 300                         | 0.3                                        | 0.2                   | 0.02                 |
|                                  | AlCl <sub>3</sub> /He (S-side: 0.01 μm)                           |                             |                                            |                       |                      |
|                                  | 80→15** (UL-side: 0.01 μm)                                        |                             |                                            |                       |                      |
|                                  | 15→5**                                                            |                             |                                            |                       |                      |
| Upper layer                      | SiH <sub>4</sub> 40                                               |                             |                                            |                       |                      |
| 1st layer region                 | H <sub>2</sub> 200                                                | 300                         | 5                                          | 0.2                   | 10                   |
|                                  | B <sub>2</sub> H <sub>6</sub> (against SiH <sub>4</sub> ) 200 ppm |                             |                                            |                       |                      |
| 2nd layer region                 | SiH <sub>4</sub> 100                                              |                             |                                            |                       |                      |
|                                  | H <sub>2</sub> 300                                                | 300                         | 6                                          | 0.3                   | 20                   |
| 3rd layer region                 | SiH <sub>4</sub> 20                                               |                             |                                            |                       |                      |
|                                  | CH <sub>4</sub> 200                                               | 300                         | 3                                          | 0.2                   | 0.5                  |

TABLE 21

| Order of lamination (layer name) | Gases and their flow rates (SCCM)                                                                       | Substrate temperature (°C.) | RF discharging power (mW/cm <sup>3</sup> ) | Inner pressure (Torr) | Layer thickness (μm) |
|----------------------------------|---------------------------------------------------------------------------------------------------------|-----------------------------|--------------------------------------------|-----------------------|----------------------|
| Lower layer                      | SiH <sub>4</sub> 50                                                                                     |                             |                                            |                       |                      |
|                                  | H <sub>2</sub> 5→200*                                                                                   | 500                         | 5                                          | 0.4                   | 0.05                 |
|                                  | AlCl <sub>3</sub> /He 200→20**                                                                          |                             |                                            |                       |                      |
| Upper layer                      | SiH <sub>4</sub> 100                                                                                    |                             |                                            |                       |                      |
| 1st layer region                 | B <sub>2</sub> H <sub>6</sub> (against SiH <sub>4</sub> ) (LL-side: 2 μm) (U·2nd·LR-side: 1 μm) 500 ppm | 500                         | 20                                         | 0.4                   | 3                    |
|                                  | 500 ppm→0**                                                                                             |                             |                                            |                       |                      |
| 2nd                              | H <sub>2</sub> 1200                                                                                     |                             |                                            |                       |                      |
|                                  | SiH <sub>4</sub> 300                                                                                    |                             |                                            |                       |                      |

TABLE 21-continued

| Order of lamination (layer name) | Gases and their flow rates (SCCM) | Substrate temperature (°C.) | RF discharging power (mW/cm <sup>3</sup> ) | Inner pressure (Torr) | Layer thickness (μm) |
|----------------------------------|-----------------------------------|-----------------------------|--------------------------------------------|-----------------------|----------------------|
| layer region                     | H <sub>2</sub> 1500               | 500                         | 30                                         | 0.5                   | 10                   |
| 3rd layer region                 | SiH <sub>4</sub> 200              |                             |                                            |                       |                      |
| C <sub>2</sub> H <sub>2</sub>    | 10 → 20*                          | 500                         | 30                                         | 0.4                   | 20                   |
| NO                               | 1                                 |                             |                                            |                       |                      |

TABLE 22

| Order of lamination (layer name) | Gases and their flow rates (SCCM)                                 | Substrate temperature (°C.) | μW discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 150                                              |                             |                                            |                       |                      |
|                                  | H <sub>2</sub> 20 → 500*                                          | 250                         | 0.5                                        | 0.6                   | 0.02                 |
|                                  | AlCl <sub>3</sub> /He (S-side: 0.01 μm)                           |                             |                                            |                       |                      |
|                                  | 400 → 80** (UL-side: 0.01 μm)                                     |                             |                                            |                       |                      |
|                                  | 80 → 50**                                                         |                             |                                            |                       |                      |
| Upper layer                      | 1st layer region                                                  | SiH <sub>4</sub> 100        |                                            |                       |                      |
|                                  | B <sub>2</sub> H <sub>6</sub> (against SiH <sub>4</sub> ) 200 ppm | 250                         | 0.5                                        | 0.5                   | 3                    |
|                                  | H <sub>2</sub> 500                                                |                             |                                            |                       |                      |
|                                  | 2nd layer region                                                  | SiH <sub>4</sub> 700        |                                            |                       |                      |
|                                  | SiF <sub>4</sub> 30                                               | 250                         | 0.5                                        | 0.5                   | 20                   |
|                                  | H <sub>2</sub> 500                                                |                             |                                            |                       |                      |
|                                  | 3rd layer region                                                  | SiH <sub>4</sub> 150        |                                            |                       |                      |
|                                  | CH <sub>4</sub> 500                                               | 250                         | 0.5                                        | 0.3                   | 1                    |
|                                  | region                                                            |                             |                                            |                       |                      |

TABLE 23

| Order of lamination (layer name) | Gases and their flow rates (SCCM)                                         | Substrate temperature (°C.) | RF discharging power (mW/cm <sup>3</sup> ) | Inner pressure (Torr) | Layer thickness (μm) |
|----------------------------------|---------------------------------------------------------------------------|-----------------------------|--------------------------------------------|-----------------------|----------------------|
| Lower Layer                      | SiH <sub>4</sub> 50                                                       |                             |                                            |                       |                      |
|                                  | H <sub>2</sub> 5 → 200*                                                   | 250                         | 5                                          | 0.4                   | 0.05                 |
|                                  | AlCl <sub>3</sub> /He 200 → 20**                                          |                             |                                            |                       |                      |
| Upper layer                      | 1st layer region                                                          | SiH <sub>4</sub> 100        |                                            |                       |                      |
|                                  | B <sub>2</sub> H <sub>6</sub> (against SiH <sub>4</sub> ) (LL-side: 3 μm) | 500 ppm                     | 250                                        | 10                    | 0.4                  |
|                                  | (U · 2nd · LR-side: 2 μm)                                                 |                             | 500 ppm → 0**                              |                       |                      |
|                                  | H <sub>2</sub> 200                                                        |                             |                                            |                       |                      |
|                                  | AlCl <sub>3</sub> /He (against SiH <sub>4</sub> ) 1 → 0**                 |                             |                                            |                       |                      |
| 2nd layer region                 | SiH <sub>4</sub> 200                                                      |                             |                                            |                       |                      |
|                                  | C <sub>2</sub> H <sub>2</sub> 10 → 20*                                    | 250                         | 15                                         | 0.4                   | 20                   |
|                                  | NO 1                                                                      |                             |                                            |                       |                      |
| 3rd layer region                 | SiH <sub>4</sub> 300                                                      |                             |                                            |                       |                      |
|                                  | H <sub>2</sub> 300                                                        | 250                         | 15                                         | 0.5                   | 10                   |
|                                  | region                                                                    |                             |                                            |                       |                      |

TABLE 24

| Order of lamination (layer name) | Gases and their flow rates (SCCM)                                         | Substrate temperature (°C.) | RF discharging power (mW/cm <sup>3</sup> ) | Inner pressure (Torr) | Layer thickness (μm) |
|----------------------------------|---------------------------------------------------------------------------|-----------------------------|--------------------------------------------|-----------------------|----------------------|
| Lower layer                      | SiH <sub>4</sub> 50                                                       |                             |                                            |                       |                      |
|                                  | H <sub>2</sub> 5 → 200*                                                   | 250                         | 1                                          | 0.4                   | 0.02                 |
|                                  | AlCl <sub>3</sub> /He (S-side: 0.01 μm)                                   |                             |                                            |                       |                      |
|                                  | 200 → 30**                                                                |                             |                                            |                       |                      |
|                                  | (UL-side: 0.01 μm)                                                        |                             |                                            |                       |                      |
| Upper layer                      | 1st layer region                                                          | SiH <sub>4</sub> 100        |                                            |                       |                      |
|                                  | B <sub>2</sub> H <sub>6</sub> (against SiH <sub>4</sub> ) (LL-side: 2 μm) | 500 ppm                     | 250                                        | 10                    | 0.4                  |
|                                  | (U · 2nd · LR-side: 1 μm)                                                 |                             | 500 ppm → 0**                              |                       |                      |
|                                  | H <sub>2</sub> 200                                                        |                             |                                            |                       |                      |
| 2nd layer region                 | SiH <sub>4</sub> 100                                                      |                             |                                            |                       |                      |
|                                  | C <sub>2</sub> H <sub>2</sub> 100                                         | 300                         | 15                                         | 0.4                   | 20                   |
|                                  | NO 1                                                                      |                             |                                            |                       |                      |
| 3rd layer region                 | SiH <sub>4</sub> 300                                                      |                             |                                            |                       |                      |
|                                  | H <sub>2</sub> 300                                                        | 300                         | 20                                         | 0.5                   | 5                    |
|                                  | region                                                                    |                             |                                            |                       |                      |

TABLE 24-continued

| Order of lamination (layer name) | Gases and their flow rates (SCCM)   |           | Substrate temperature (°C.) | RF discharging power (mW/cm <sup>3</sup> ) | Inner pressure (Torr) | Layer thickness (μm) |
|----------------------------------|-------------------------------------|-----------|-----------------------------|--------------------------------------------|-----------------------|----------------------|
| region                           |                                     |           |                             |                                            |                       |                      |
| 4th layer region                 | SiH <sub>4</sub><br>CH <sub>4</sub> | 50<br>600 | 300                         | 10                                         | 0.4                   | 0.5                  |

TABLE 25

| Order of lamination (layer name) | Gases and their flow rates (SCCM)                                                |                                                                                                 | Substrate temperature (°C.) | RF discharging power (mW/cm <sup>3</sup> ) | Inner pressure (Torr) | Layer thickness (μm) |
|----------------------------------|----------------------------------------------------------------------------------|-------------------------------------------------------------------------------------------------|-----------------------------|--------------------------------------------|-----------------------|----------------------|
| Lower layer                      | SiH <sub>4</sub><br>H <sub>2</sub><br>AlCl <sub>3</sub> /He<br>(S-side: 0.05 μm) | 10 → 100*<br>5 → 200*<br>200 → 40**<br>(UL-side: 0.15 μm)                                       | 300                         | 5                                          | 0.4                   | 0.2                  |
| Upper layer                      | 1st layer region                                                                 | SiH <sub>4</sub><br>B <sub>2</sub> H <sub>6</sub> (against SiH <sub>4</sub> )<br>H <sub>2</sub> | 100<br>200 ppm<br>500       | 300                                        | 5                     | 0.4                  |
| 2nd layer region                 | SiH <sub>4</sub><br>NH <sub>3</sub>                                              | 300<br>50                                                                                       | 300                         | 15                                         | 0.4                   | 25                   |
| 3rd layer region                 | SiH <sub>4</sub><br>H <sub>2</sub>                                               | 100<br>300                                                                                      | 300                         | 5                                          | 0.2                   | 8                    |
| 4th layer region                 | SiH <sub>4</sub><br>NH <sub>3</sub>                                              | 100<br>50                                                                                       | 300                         | 10                                         | 0.4                   | 0.3                  |

TABLE 26

| Order of lamination (layer name) | Gases and their flow rates (SCCM)                                                |                                                                                   | Substrate temperature (°C.) | RF discharging power (mW/cm <sup>3</sup> ) | Inner pressure (Torr) | Layer thickness (μm) |
|----------------------------------|----------------------------------------------------------------------------------|-----------------------------------------------------------------------------------|-----------------------------|--------------------------------------------|-----------------------|----------------------|
| Lower layer                      | SiH <sub>4</sub><br>H <sub>2</sub><br>AlCl <sub>3</sub> /He<br>(S-side: 0.05 μm) | 10 → 100*<br>5 → 200*<br>200 → 40**<br>(UL-side: 0.15 μm)                         | 250                         | 5                                          | 0.4                   | 0.2                  |
| Upper layer                      | 1st layer region                                                                 | SiH <sub>4</sub><br>PH <sub>3</sub> (against SiH <sub>4</sub> )<br>H <sub>2</sub> | 100<br>100 ppm<br>100       | 250                                        | 8                     | 0.4                  |
| 2nd layer region                 | SiH <sub>4</sub><br>CH <sub>4</sub>                                              | 100<br>100                                                                        | 300                         | 15                                         | 0.4                   | 30                   |
| 3rd layer region                 | SiH <sub>4</sub><br>SiF <sub>4</sub>                                             | 100<br>5                                                                          | 300                         | 3                                          | 0.5                   | 3                    |
| 4th layer region                 | H <sub>2</sub><br>SiH <sub>4</sub>                                               | 200<br>50                                                                         | 300                         | 10                                         | 0.4                   | 0.5                  |
|                                  |                                                                                  | 600                                                                               |                             |                                            |                       |                      |

TABLE 27

| Order of lamination (layer name) | Gases and their flow rates (SCCM)                                                                                                                             |                                                                                                                               | Substrate temperature (°C.) | RF discharging power (mW/cm <sup>3</sup> ) | Inner pressure (Torr) | Layer thickness (μm) |
|----------------------------------|---------------------------------------------------------------------------------------------------------------------------------------------------------------|-------------------------------------------------------------------------------------------------------------------------------|-----------------------------|--------------------------------------------|-----------------------|----------------------|
| Lower layer                      | SiH <sub>4</sub><br>H <sub>2</sub><br>AlCl <sub>3</sub> /He                                                                                                   | 50<br>5 → 200*<br>200 → 20**                                                                                                  | 250                         | 5                                          | 0.4                   | 0.05                 |
| Upper layer                      | 1st layer region                                                                                                                                              | SiH <sub>4</sub><br>B <sub>2</sub> H <sub>6</sub> (against SiH <sub>4</sub> )<br>(LL-side: 2 μm)<br>(U · 2nd · LR-side: 1 μm) | 100<br>500 ppm              | 250                                        | 8                     | 0.4                  |
| 2nd layer region                 | H <sub>2</sub><br>SiH <sub>4</sub><br>C <sub>2</sub> H <sub>2</sub><br>B <sub>2</sub> H <sub>6</sub> (against SiH <sub>4</sub> )<br>(U · 1st · LR-side: 1 μm) | 200<br>300<br>50<br>0 → 100 ppm*                                                                                              | 330                         | 20                                         | 0.4                   | 30                   |

TABLE 27-continued

| Order of lamination (layer name) | Gases and their flow rates (SCCM) | Substrate temperature (°C.) | RF discharging power (mW/cm <sup>3</sup> ) | Inner pressure (Torr) | Layer thickness (μm) |
|----------------------------------|-----------------------------------|-----------------------------|--------------------------------------------|-----------------------|----------------------|
| (U · 3rd · LR-side: 29 μm)       |                                   |                             |                                            |                       |                      |
| 3rd layer region                 | Si <sub>2</sub> H <sub>6</sub>    | 100 ppm                     |                                            |                       |                      |
|                                  | H <sub>2</sub>                    | 200                         |                                            |                       |                      |
| 4th layer region                 | SiH <sub>4</sub>                  | 200                         |                                            |                       |                      |
|                                  | C <sub>2</sub> H <sub>2</sub>     | 200                         | 330                                        | 10                    | 0.4                  |
|                                  |                                   |                             |                                            |                       | 1                    |

TABLE 28

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 10 → 100*                   |                                            |                       |                      |
|                                  | H <sub>2</sub>                                            | 5 → 200*                    |                                            |                       |                      |
|                                  | AlCl <sub>3</sub> /He (S-side: 0.05 μm)                   | 250                         | 5                                          | 0.4                   | 0.2                  |
|                                  | (UL-side: 0.15 μm)                                        |                             |                                            |                       |                      |
| Upper layer                      | SiH <sub>4</sub>                                          | 200 → 40**                  |                                            |                       |                      |
|                                  | H <sub>2</sub>                                            | 40                          |                                            |                       |                      |
| 1st layer region                 | PH <sub>3</sub> (against SiH <sub>4</sub> )               | 250 ppm                     | 250                                        | 8                     | 0.4                  |
|                                  | (LL-side: 2 μm)                                           |                             |                                            |                       | 3                    |
|                                  | (U · 2nd · LR-side: 1 μm)                                 |                             |                                            |                       |                      |
| 2nd layer region                 | H <sub>2</sub>                                            | 250 ppm → 0**               |                                            |                       |                      |
|                                  | SiH <sub>4</sub>                                          | 40                          |                                            |                       |                      |
| 3rd layer region                 | NH <sub>3</sub>                                           | 300                         |                                            |                       |                      |
|                                  | PH <sub>3</sub> (against SiH <sub>4</sub> )               | 30 → 50*                    | 300                                        | 15                    | 0.4                  |
| 4th layer region                 | SiH <sub>4</sub>                                          | 50 ppm                      |                                            |                       |                      |
|                                  | H <sub>2</sub>                                            | 100                         | 300                                        | 5                     | 0.2                  |
| 5th layer region                 | SiH <sub>4</sub>                                          | 300                         |                                            |                       |                      |
|                                  | NH <sub>3</sub>                                           | 100                         | 300                                        | 5                     | 0.4                  |
|                                  | B <sub>2</sub> H <sub>6</sub> (against SiH <sub>4</sub> ) | 80 → 100*                   |                                            |                       | 0.7                  |
|                                  |                                                           | 500 ppm                     |                                            |                       |                      |

TABLE 29

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 50                          |                                            |                       |                      |
|                                  | H <sub>2</sub>                                            | 5 → 200*                    |                                            |                       |                      |
|                                  | AlCl <sub>3</sub> /He (S-side: 0.01 μm)                   | 250                         | 1                                          | 0.3                   | 0.02                 |
|                                  | (UL-side: 0.01 μm)                                        |                             |                                            |                       |                      |
| Upper layer                      | SiH <sub>4</sub>                                          | 200 → 30**                  |                                            |                       |                      |
|                                  | B <sub>2</sub> H <sub>6</sub> (against SiH <sub>4</sub> ) | 100                         | 250                                        | 10                    | 0.4                  |
| 1st layer region                 | He                                                        | 500 ppm                     | 250                                        | 10                    | 0.4                  |
| 2nd layer region                 | SiH <sub>4</sub>                                          | 600                         | 250                                        | 25                    | 0.6                  |
| 3rd layer region                 | B <sub>2</sub> H <sub>6</sub>                             | 600                         |                                            |                       |                      |
| 4th layer region                 | SiH <sub>4</sub>                                          | 0.5 ppm                     |                                            |                       |                      |
| 5th layer region                 | CH <sub>4</sub>                                           | 50                          | 250                                        | 10                    | 0.4                  |
|                                  |                                                           | 500                         |                                            |                       | 1                    |

TABLE 30

| Order of lamination (layer name) | Gases and their flow rates (SCCM)       | Substrate temperature (°C.) | RF discharging power (mW/cm <sup>3</sup> ) | Inner pressure (Torr) | Layer thickness (μm) |
|----------------------------------|-----------------------------------------|-----------------------------|--------------------------------------------|-----------------------|----------------------|
| Lower layer                      | SiH <sub>4</sub>                        | 10 → 100*                   |                                            |                       |                      |
|                                  | H <sub>2</sub>                          | 5 → 200*                    |                                            |                       |                      |
|                                  | AlCl <sub>3</sub> /He (S-side: 0.05 μm) | 300                         | 10                                         | 0.4                   | 0.2                  |
|                                  | (UL-side: 0.15 μm)                      |                             |                                            |                       |                      |
| Upper layer                      | SiH <sub>4</sub>                        | 200 → 40**                  |                                            |                       |                      |
|                                  | B <sub>2</sub> H <sub>6</sub>           | 100                         |                                            |                       |                      |
| 1st layer region                 | He                                      | 200 ppm                     | 300                                        | 8                     | 0.4                  |
| 2nd layer region                 | SiH <sub>4</sub>                        | 500                         |                                            |                       | 0.5                  |

TABLE 30-continued

| Order of lamination (layer name) | Gases and their flow rates (SCCM)                    | Substrate temperature (°C.) | RF discharging power (mW/cm <sup>3</sup> ) | Inner pressure (Torr) | Layer thickness (μm) |
|----------------------------------|------------------------------------------------------|-----------------------------|--------------------------------------------|-----------------------|----------------------|
| 2nd layer region                 | SiF <sub>4</sub> 0.5                                 |                             |                                            |                       |                      |
|                                  | AlCl <sub>3</sub> /He 0.1                            |                             |                                            |                       |                      |
|                                  | SiH <sub>4</sub> 300                                 |                             |                                            |                       |                      |
|                                  | H <sub>2</sub> 500                                   |                             |                                            |                       |                      |
|                                  | CH <sub>4</sub> 1                                    | 300                         | 20                                         | 0.5                   | 20                   |
|                                  | NO 0.1                                               |                             |                                            |                       |                      |
|                                  | B <sub>2</sub> H <sub>6</sub> 0.3 ppm                |                             |                                            |                       |                      |
|                                  | SiF <sub>4</sub> 0.5                                 |                             |                                            |                       |                      |
|                                  | AlCl <sub>3</sub> /He 0.1                            |                             |                                            |                       |                      |
| 3rd layer region                 | SiH <sub>4</sub> 100                                 |                             |                                            |                       |                      |
|                                  | CH <sub>4</sub> 600                                  |                             |                                            |                       |                      |
|                                  | PH <sub>3</sub> (against SiH <sub>4</sub> ) 3000 ppm | 300                         | 15                                         | 0.4                   | 7                    |
|                                  | NO 0.1                                               |                             |                                            |                       |                      |
|                                  | SiF <sub>4</sub> 0.5                                 |                             |                                            |                       |                      |
|                                  | AlCl <sub>3</sub> /He 0.1                            |                             |                                            |                       |                      |
|                                  | B <sub>2</sub> H <sub>6</sub> 0.3 ppm                |                             |                                            |                       |                      |
|                                  | SiH <sub>4</sub> 40                                  |                             |                                            |                       |                      |
|                                  | CH <sub>4</sub> 600                                  |                             |                                            |                       |                      |
| 4th layer region                 | NO 0.1                                               | 300                         | 10                                         | 0.4                   | 0.1                  |
|                                  | PH <sub>3</sub> 0.3 ppm                              |                             |                                            |                       |                      |
|                                  | B <sub>2</sub> H <sub>6</sub> 0.3 ppm                |                             |                                            |                       |                      |
|                                  | SiF <sub>4</sub> 0.5                                 |                             |                                            |                       |                      |
|                                  | AlCl <sub>3</sub> /He 0.1                            |                             |                                            |                       |                      |
|                                  | SiH <sub>4</sub>                                     |                             |                                            |                       |                      |
|                                  | CH <sub>4</sub>                                      |                             |                                            |                       |                      |
|                                  | NO                                                   |                             |                                            |                       |                      |
|                                  | SiF <sub>4</sub>                                     |                             |                                            |                       |                      |

TABLE 31

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 10 → 100*                                        |                             |                                            |                       |                      |
|                                  | H <sub>2</sub> 5 → 200*                                           |                             |                                            |                       |                      |
|                                  | AlCl <sub>3</sub> /He (S-side: 0.05 μm)                           | 250                         | 5                                          | 0.4                   | 0.2                  |
|                                  | 200 → 40** (UL-side: 0.15 μm)                                     |                             |                                            |                       |                      |
|                                  | 40 → 10**                                                         |                             |                                            |                       |                      |
|                                  | SiH <sub>4</sub> 100                                              |                             |                                            |                       |                      |
|                                  | B <sub>2</sub> H <sub>6</sub> (against SiH <sub>4</sub> ) 500 ppm | 250                         | 8                                          | 0.4                   | 3                    |
|                                  | (LL-side: 2 μm) (U · 2nd · LR-side: 1 μm) 500 ppm → 0**           |                             |                                            |                       |                      |
|                                  | H <sub>2</sub> 200                                                |                             |                                            |                       |                      |
| Upper layer                      | SiF <sub>4</sub> 0.5                                              |                             |                                            |                       |                      |
|                                  | AlCl <sub>3</sub> /He 0.1                                         |                             |                                            |                       |                      |
|                                  | SiH <sub>4</sub> 100                                              |                             |                                            |                       |                      |
|                                  | SiF <sub>4</sub> 5                                                |                             |                                            |                       |                      |
|                                  | H <sub>2</sub> 200                                                | 300                         | 3                                          | 0.5                   | 3                    |
|                                  | CH <sub>4</sub> 1                                                 |                             |                                            |                       |                      |
|                                  | NO 0.1                                                            |                             |                                            |                       |                      |
|                                  | B <sub>2</sub> H <sub>6</sub> (against SiH <sub>4</sub> ) 0.3 ppm |                             |                                            |                       |                      |
|                                  | AlCl <sub>3</sub> /He 0.1                                         |                             |                                            |                       |                      |
| 1st layer region                 | SiH <sub>4</sub> 100                                              |                             |                                            |                       |                      |
|                                  | CH <sub>4</sub> 100                                               |                             |                                            |                       |                      |
|                                  | PH <sub>3</sub> (against SiH <sub>4</sub> ) 50 ppm                | 300                         | 15                                         | 0.4                   | 30                   |
|                                  | NO 0.1                                                            |                             |                                            |                       |                      |
|                                  | B <sub>2</sub> H <sub>6</sub> (against SiH <sub>4</sub> ) 0.3 ppm |                             |                                            |                       |                      |
|                                  | SiF <sub>4</sub> 0.5                                              |                             |                                            |                       |                      |
|                                  | AlCl <sub>3</sub> /He 0.1                                         |                             |                                            |                       |                      |
|                                  | SiH <sub>4</sub> 50                                               |                             |                                            |                       |                      |
|                                  | CH <sub>4</sub> 600                                               |                             |                                            |                       |                      |
| 2nd layer region                 | PH <sub>3</sub> (against SiH <sub>4</sub> ) 0.3 ppm               | 300                         | 10                                         | 0.4                   | 0.5                  |
|                                  | B <sub>2</sub> H <sub>6</sub> (against SiH <sub>4</sub> ) 0.3 ppm |                             |                                            |                       |                      |
|                                  | NO 0.1                                                            |                             |                                            |                       |                      |
|                                  | SiF <sub>4</sub> 0.5                                              |                             |                                            |                       |                      |
|                                  | AlCl <sub>3</sub> /He 0.1                                         |                             |                                            |                       |                      |
|                                  | SiH <sub>4</sub>                                                  |                             |                                            |                       |                      |
|                                  | CH <sub>4</sub>                                                   |                             |                                            |                       |                      |
|                                  | NO                                                                |                             |                                            |                       |                      |
|                                  | SiF <sub>4</sub>                                                  |                             |                                            |                       |                      |
| 3rd layer region                 | AlCl <sub>3</sub> /He 0.1                                         |                             |                                            |                       |                      |
|                                  | SiH <sub>4</sub> 100                                              |                             |                                            |                       |                      |
|                                  | CH <sub>4</sub> 100                                               |                             |                                            |                       |                      |
|                                  | PH <sub>3</sub> (against SiH <sub>4</sub> ) 50 ppm                | 300                         | 15                                         | 0.4                   | 30                   |
|                                  | NO 0.1                                                            |                             |                                            |                       |                      |
|                                  | B <sub>2</sub> H <sub>6</sub> (against SiH <sub>4</sub> ) 0.3 ppm |                             |                                            |                       |                      |
|                                  | SiF <sub>4</sub> 0.5                                              |                             |                                            |                       |                      |
|                                  | AlCl <sub>3</sub> /He 0.1                                         |                             |                                            |                       |                      |
|                                  | SiH <sub>4</sub>                                                  |                             |                                            |                       |                      |
| 4th layer region                 | CH <sub>4</sub> 50                                                |                             |                                            |                       |                      |
|                                  | NO 0.1                                                            |                             |                                            |                       |                      |
|                                  | SiF <sub>4</sub> 0.5                                              |                             |                                            |                       |                      |
|                                  | AlCl <sub>3</sub> /He 0.1                                         |                             |                                            |                       |                      |
|                                  | SiH <sub>4</sub>                                                  |                             |                                            |                       |                      |
|                                  | CH <sub>4</sub>                                                   |                             |                                            |                       |                      |
|                                  | NO                                                                |                             |                                            |                       |                      |
|                                  | SiF <sub>4</sub>                                                  |                             |                                            |                       |                      |
|                                  | AlCl <sub>3</sub> /He                                             |                             |                                            |                       |                      |

TABLE 32

| Order of lamination (layer name) | Gases and their flow rates (SCCM)       | Substrate temperature (°C.) | RF discharging power (mW/cm <sup>3</sup> ) | Inner pressure (Torr) | Layer thickness (μm) |
|----------------------------------|-----------------------------------------|-----------------------------|--------------------------------------------|-----------------------|----------------------|
| Lower layer                      | SiH <sub>4</sub> 10 → 100*              |                             |                                            |                       |                      |
|                                  | H <sub>2</sub> 5 → 200*                 |                             |                                            |                       |                      |
|                                  | AlCl <sub>3</sub> /He (S-side: 0.05 μm) | 300                         | 10                                         | 0.4                   | 0.2                  |
|                                  | 200 → 40**                              |                             |                                            |                       |                      |
|                                  | SiH <sub>4</sub>                        |                             |                                            |                       |                      |
|                                  | CH <sub>4</sub>                         |                             |                                            |                       |                      |
|                                  | NO                                      |                             |                                            |                       |                      |
|                                  | SiF <sub>4</sub>                        |                             |                                            |                       |                      |
|                                  | AlCl <sub>3</sub> /He                   |                             |                                            |                       |                      |

TABLE 32-continued

| Order of lamination<br>(layer name) | Gases and their flow rates<br>(SCCM)        | Substrate temperature<br>(°C.) | RF discharging power<br>(mW/cm <sup>3</sup> ) | Inner pressure<br>(Torr) | Layer thickness<br>(μm) |
|-------------------------------------|---------------------------------------------|--------------------------------|-----------------------------------------------|--------------------------|-------------------------|
| (UL-side: 0.15 μm)                  |                                             |                                |                                               |                          |                         |
| Upper layer                         | SiH <sub>4</sub>                            | 100                            | 300                                           | 8                        | 0.5                     |
|                                     | B <sub>2</sub> H <sub>6</sub>               | 200 ppm                        |                                               |                          |                         |
|                                     | H <sub>2</sub>                              | 500                            |                                               |                          |                         |
|                                     | SiF <sub>4</sub>                            | 0.5                            |                                               |                          |                         |
|                                     | AlCl <sub>3</sub> /He                       | 0.1                            |                                               |                          |                         |
|                                     | H <sub>2</sub> S                            | 1 ppm                          |                                               |                          |                         |
|                                     | SiH <sub>4</sub>                            | 300                            |                                               |                          |                         |
|                                     | H <sub>2</sub>                              | 500                            |                                               |                          |                         |
|                                     | CH <sub>4</sub>                             | 1                              |                                               |                          |                         |
|                                     | NO                                          | 0.1                            |                                               |                          |                         |
| 2nd layer                           | B <sub>2</sub> H <sub>6</sub>               | 0.3 ppm                        |                                               |                          |                         |
|                                     | SiF <sub>4</sub>                            | 0.5                            |                                               |                          |                         |
|                                     | AlCl <sub>3</sub> /He                       | 0.1                            |                                               |                          |                         |
|                                     | H <sub>2</sub> S                            | 1 ppm                          |                                               |                          |                         |
|                                     | SiH <sub>4</sub>                            | 100                            |                                               |                          |                         |
|                                     | CH <sub>4</sub>                             | 600                            |                                               |                          |                         |
|                                     | PH <sub>3</sub> (against SiH <sub>4</sub> ) | 3000 ppm                       |                                               |                          |                         |
|                                     | NO                                          | 0.1                            |                                               |                          |                         |
|                                     | SiF <sub>4</sub>                            | 0.5                            |                                               |                          |                         |
|                                     | AlCl <sub>3</sub> /He                       | 0.1                            |                                               |                          |                         |
| 3rd layer                           | B <sub>2</sub> H <sub>6</sub>               | 0.3 ppm                        |                                               |                          |                         |
|                                     | SiH <sub>4</sub>                            | 100                            |                                               |                          |                         |
|                                     | CH <sub>4</sub>                             | 600                            |                                               |                          |                         |
|                                     | NO                                          | 0.1                            |                                               |                          |                         |
|                                     | SiF <sub>4</sub>                            | 0.5                            |                                               |                          |                         |
|                                     | AlCl <sub>3</sub> /He                       | 0.1                            |                                               |                          |                         |
|                                     | H <sub>2</sub> S                            | 1 ppm                          |                                               |                          |                         |
|                                     | SiH <sub>4</sub>                            | 40                             |                                               |                          |                         |
|                                     | CH <sub>4</sub>                             | 600                            |                                               |                          |                         |
|                                     | NO                                          | 0.1                            |                                               |                          |                         |
| 4th layer                           | PH <sub>3</sub>                             | 0.3 ppm                        |                                               |                          |                         |
|                                     | B <sub>2</sub> H <sub>6</sub>               | 0.3 ppm                        |                                               |                          |                         |
|                                     | SiF <sub>4</sub>                            | 0.5                            |                                               |                          |                         |
|                                     | AlCl <sub>3</sub> /He                       | 0.1                            |                                               |                          |                         |
|                                     | H <sub>2</sub> S                            | 1 ppm                          |                                               |                          |                         |
|                                     | SiH <sub>4</sub>                            | 40                             |                                               |                          |                         |
|                                     | CH <sub>4</sub>                             | 600                            |                                               |                          |                         |
|                                     | NO                                          | 0.1                            |                                               |                          |                         |
|                                     | PH <sub>3</sub>                             | 0.3 ppm                        |                                               |                          |                         |
|                                     | B <sub>2</sub> H <sub>6</sub>               | 0.3 ppm                        |                                               |                          |                         |

TABLE 33

| Order of lamination<br>(layer name) | Gases and their flow rates<br>(SCCM)                      | Substrate temperature<br>(°C.) | RF discharging power<br>(mW/cm <sup>3</sup> ) | Inner pressure<br>(Torr) | Layer thickness<br>(μm) |
|-------------------------------------|-----------------------------------------------------------|--------------------------------|-----------------------------------------------|--------------------------|-------------------------|
| Lower layer                         | SiH <sub>4</sub>                                          | 50                             | 250                                           | 5                        | 0.4                     |
|                                     | H <sub>2</sub>                                            | 10 → *                         |                                               |                          |                         |
|                                     | AlCl <sub>3</sub> /He                                     | 120 → 40**                     |                                               |                          |                         |
|                                     | B <sub>2</sub> H <sub>6</sub> (against SiH <sub>4</sub> ) | 100 ppm                        |                                               |                          |                         |
|                                     | SiH <sub>4</sub>                                          | 100                            |                                               |                          |                         |
|                                     | B <sub>2</sub> H <sub>6</sub> (against SiH <sub>4</sub> ) | 200 ppm                        |                                               |                          |                         |
|                                     | H <sub>2</sub>                                            | 500                            |                                               |                          |                         |
|                                     | SiH <sub>4</sub>                                          | 300                            |                                               |                          |                         |
|                                     | H <sub>2</sub>                                            | 300                            |                                               |                          |                         |
|                                     | SiH <sub>4</sub>                                          | 50                             |                                               |                          |                         |
| Upper layer                         | CH <sub>4</sub>                                           | 500                            |                                               |                          |                         |
|                                     | SiH <sub>4</sub>                                          | 250                            |                                               |                          |                         |
|                                     | NO                                                        | 0.1                            |                                               |                          |                         |
|                                     | SiF <sub>4</sub>                                          | 0.5                            |                                               |                          |                         |
|                                     | AlCl <sub>3</sub> /He                                     | 0.1                            |                                               |                          |                         |
|                                     | H <sub>2</sub> S                                          | 1 ppm                          |                                               |                          |                         |
|                                     | SiH <sub>4</sub>                                          | 40                             |                                               |                          |                         |
|                                     | CH <sub>4</sub>                                           | 600                            |                                               |                          |                         |
|                                     | NO                                                        | 0.1                            |                                               |                          |                         |
|                                     | PH <sub>3</sub>                                           | 0.3 ppm                        |                                               |                          |                         |

TABLE 34

| Order of lamination<br>(layer name) | Gases and their flow rates<br>(SCCM)                      | Substrate temperature<br>(°C.) | RF discharging power<br>(mW/cm <sup>3</sup> ) | Inner pressure<br>(Torr) | Layer thickness<br>(μm) |
|-------------------------------------|-----------------------------------------------------------|--------------------------------|-----------------------------------------------|--------------------------|-------------------------|
| Lower layer                         | SiH <sub>4</sub>                                          | 50                             | 250                                           | 5                        | 0.05                    |
|                                     | AlCl <sub>3</sub> /He                                     | 120 → 40**                     |                                               |                          |                         |
|                                     | SiH <sub>4</sub>                                          | 100                            |                                               |                          |                         |
|                                     | B <sub>2</sub> H <sub>6</sub> (against SiH <sub>4</sub> ) | 200 ppm                        |                                               |                          |                         |
|                                     | H <sub>2</sub>                                            | 500                            |                                               |                          |                         |
|                                     | SiH <sub>4</sub>                                          | 300                            |                                               |                          |                         |
|                                     | H <sub>2</sub>                                            | 300                            |                                               |                          |                         |
|                                     | SiH <sub>4</sub>                                          | 50                             |                                               |                          |                         |
|                                     | CH <sub>4</sub>                                           | 500                            |                                               |                          |                         |
|                                     | NO                                                        | 0.1                            |                                               |                          |                         |
| Upper layer                         | SiH <sub>4</sub>                                          | 250                            | 8                                             | 0.4                      | 3                       |
|                                     | NO                                                        | 0.1                            |                                               |                          |                         |
|                                     | SiF <sub>4</sub>                                          | 0.5                            |                                               |                          |                         |
|                                     | AlCl <sub>3</sub> /He                                     | 0.1                            |                                               |                          |                         |
|                                     | H <sub>2</sub> S                                          | 1 ppm                          |                                               |                          |                         |
|                                     | SiH <sub>4</sub>                                          | 100                            |                                               |                          |                         |
|                                     | B <sub>2</sub> H <sub>6</sub> (against SiH <sub>4</sub> ) | 200 ppm                        |                                               |                          |                         |
|                                     | H <sub>2</sub>                                            | 500                            |                                               |                          |                         |
|                                     | SiH <sub>4</sub>                                          | 300                            |                                               |                          |                         |
|                                     | H <sub>2</sub>                                            | 300                            |                                               |                          |                         |
| 2nd layer                           | SiH <sub>4</sub>                                          | 250                            | 15                                            | 0.5                      | 20                      |
|                                     | NO                                                        | 0.1                            |                                               |                          |                         |
|                                     | SiF <sub>4</sub>                                          | 0.5                            |                                               |                          |                         |
|                                     | AlCl <sub>3</sub> /He                                     | 0.1                            |                                               |                          |                         |
|                                     | H <sub>2</sub> S                                          | 1 ppm                          |                                               |                          |                         |
|                                     | SiH <sub>4</sub>                                          | 50                             |                                               |                          |                         |
|                                     | CH <sub>4</sub>                                           | 500                            |                                               |                          |                         |
|                                     | NO                                                        | 0.1                            |                                               |                          |                         |
|                                     | SiF <sub>4</sub>                                          | 0.5                            |                                               |                          |                         |
|                                     | AlCl <sub>3</sub> /He                                     | 0.1                            |                                               |                          |                         |
| 3rd layer                           | SiH <sub>4</sub>                                          | 250                            | 10                                            | 0.4                      | 0.5                     |
|                                     | NO                                                        | 0.1                            |                                               |                          |                         |
|                                     | SiF <sub>4</sub>                                          | 0.5                            |                                               |                          |                         |
|                                     | AlCl <sub>3</sub> /He                                     | 0.1                            |                                               |                          |                         |
|                                     | H <sub>2</sub> S                                          | 1 ppm                          |                                               |                          |                         |
|                                     | SiH <sub>4</sub>                                          | 50                             |                                               |                          |                         |
|                                     | CH <sub>4</sub>                                           | 500                            |                                               |                          |                         |
|                                     | NO                                                        | 0.1                            |                                               |                          |                         |
|                                     | SiF <sub>4</sub>                                          | 0.5                            |                                               |                          |                         |
|                                     | AlCl <sub>3</sub> /He                                     | 0.1                            |                                               |                          |                         |
| 4th layer                           | SiH <sub>4</sub>                                          | 250                            | 10                                            | 0.4                      | 0.5                     |
|                                     | NO                                                        | 0.1                            |                                               |                          |                         |
|                                     | SiF <sub>4</sub>                                          | 0.5                            |                                               |                          |                         |
|                                     | AlCl <sub>3</sub> /He                                     | 0.1                            |                                               |                          |                         |
|                                     | H <sub>2</sub> S                                          | 1 ppm                          |                                               |                          |                         |
|                                     | SiH <sub>4</sub>                                          | 50                             |                                               |                          |                         |
|                                     | CH <sub>4</sub>                                           | 500                            |                                               |                          |                         |
|                                     | NO                                                        | 0.1                            |                                               |                          |                         |
|                                     | SiF <sub>4</sub>                                          | 0.5                            |                                               |                          |                         |
|                                     | AlCl <sub>3</sub> /He                                     | 0.1                            |                                               |                          |                         |

TABLE 35

| Order of lamination (layer name) | Gases and their flow rates (SCCM)                                                                                                                                  | Substrate temperature (°C.)      | RF discharging power (mW/cm <sup>3</sup> ) | Inner pressure (Torr) | Layer thickness (μm) |
|----------------------------------|--------------------------------------------------------------------------------------------------------------------------------------------------------------------|----------------------------------|--------------------------------------------|-----------------------|----------------------|
| Lower layer                      | SiH <sub>4</sub> 50<br>B <sub>2</sub> H <sub>6</sub> (against SiH <sub>4</sub> ) 100 ppm<br>H <sub>2</sub> 10 → 200*<br>AlCl <sub>3</sub> /He<br>(S-side: 0.01 μm) | 250                              | 5                                          | 0.4                   | 0.03                 |
|                                  |                                                                                                                                                                    | 100 → 10**<br>(UL-side: 0.01 μm) |                                            |                       |                      |
| Upper layer                      | SiH <sub>4</sub> 100<br>B <sub>2</sub> H <sub>6</sub> (against SiH <sub>4</sub> ) 200 ppm<br>H <sub>2</sub> 500<br>SiH <sub>4</sub> 300<br>H <sub>2</sub> 300      | 250                              | 8                                          | 0.4                   | 3                    |
| 1st layer region                 | SiH <sub>4</sub> 50<br>CH <sub>4</sub> 500                                                                                                                         | 250                              | 15                                         | 0.5                   | 20                   |
| 2nd layer region                 |                                                                                                                                                                    |                                  |                                            |                       |                      |
| 3rd layer region                 |                                                                                                                                                                    |                                  |                                            |                       |                      |

TABLE 36

| Order of lamination (layer name) | Gases and their flow rates (SCCM)                                                                                                                                                                      | Substrate temperature (°C.)                                 | RF discharging power (mW/cm <sup>3</sup> ) | Inner pressure (Torr) | Layer thickness (μm) |
|----------------------------------|--------------------------------------------------------------------------------------------------------------------------------------------------------------------------------------------------------|-------------------------------------------------------------|--------------------------------------------|-----------------------|----------------------|
| Lower layer                      | SiH <sub>4</sub> 50<br>H <sub>2</sub> 5 → 200*<br>AlCl <sub>3</sub> /He<br>(S-side: 0.01 μm)                                                                                                           | 150<br>↓<br>300                                             | 0.5<br>↓<br>1.5                            | 0.3                   | 0.02                 |
|                                  |                                                                                                                                                                                                        | 200 → 30**<br>(UL-side: 0.01 μm)                            |                                            |                       |                      |
| Upper layer                      | B <sub>2</sub> H <sub>6</sub> (against SiH <sub>4</sub> ) 100 ppm<br>SiH <sub>4</sub> 100<br>B <sub>2</sub> H <sub>6</sub> (against SiH <sub>4</sub> )<br>(LL-side: 2 μm)<br>(U · 2nd · LR-side: 1 μm) | 500 ppm                                                     | 250                                        | 10                    | 0.4                  |
| 1st layer region                 |                                                                                                                                                                                                        | 500 ppm → 0**<br>H <sub>2</sub> 200<br>SiH <sub>4</sub> 300 |                                            |                       | 3                    |
| 2nd layer region                 | H <sub>2</sub> 500                                                                                                                                                                                     | 250                                                         | 20                                         | 0.5                   | 20                   |

TABLE 37

| Order of lamination (layer name) | Gases and their flow rates (SCCM)                                                                                                                                                                                             | Substrate temperature (°C.)      | RF discharging power (mW/cm <sup>3</sup> ) | Inner pressure (Torr) | Layer thickness (μm) |
|----------------------------------|-------------------------------------------------------------------------------------------------------------------------------------------------------------------------------------------------------------------------------|----------------------------------|--------------------------------------------|-----------------------|----------------------|
| Lower layer                      | SiH <sub>4</sub> 50<br>H <sub>2</sub> 5 → 200*<br>AlCl <sub>3</sub> /He<br>(S-side: 0.01 μm)                                                                                                                                  | 250                              | 1                                          | 0.3                   | 0.02                 |
|                                  |                                                                                                                                                                                                                               | 200 → 30**<br>(UL-side: 0.01 μm) |                                            |                       |                      |
| 1st layer region                 | B <sub>2</sub> H <sub>6</sub> (against SiH <sub>4</sub> ) 100 ppm<br>SiH <sub>4</sub> 100<br>B <sub>2</sub> H <sub>6</sub> (against SiH <sub>4</sub> ) 500 ppm<br>He 600<br>AlCl <sub>3</sub> /He 0.1<br>SiF <sub>4</sub> 0.5 | 250                              | 10                                         | 0.4                   | 3                    |
| Upper layer                      | NO 0.1<br>CH <sub>4</sub> 1<br>2nd layer region                                                                                                                                                                               | 250                              | 25                                         | 0.6                   | 25                   |
|                                  | B <sub>2</sub> H <sub>6</sub> 0.3 ppm<br>SiF <sub>4</sub> 0.5<br>AlCl <sub>3</sub> /He 0.1<br>SiH <sub>4</sub> 50                                                                                                             |                                  |                                            |                       |                      |
| 3rd layer region                 | CH <sub>4</sub> 500<br>NO 0.1<br>B <sub>2</sub> H <sub>6</sub> 0.3 ppm<br>SiF <sub>4</sub> 0.5<br>AlCl <sub>3</sub> /He 0.1                                                                                                   | 250                              | 10                                         | 0.4                   | 1                    |

TABLE 38

| Order of lamination (layer name) | Gases and their flow rates (SCCM)                                                                     | Substrate temperature (°C.) | RF discharging power (mW/cm <sup>3</sup> ) | Inner pressure (Torr) | Layer thickness (μm) |
|----------------------------------|-------------------------------------------------------------------------------------------------------|-----------------------------|--------------------------------------------|-----------------------|----------------------|
| Lower layer                      | SiH <sub>4</sub> 10→100                                                                               | 250                         | 10                                         | 0.4                   | 0.2                  |
|                                  | H <sub>2</sub> 5→200*                                                                                 |                             |                                            |                       |                      |
|                                  | AlCl <sub>3</sub> /He (S-side:0.05 μm)                                                                |                             |                                            |                       |                      |
|                                  | 200→40** (UL-side:0.15 μm)                                                                            |                             |                                            |                       |                      |
|                                  | B <sub>2</sub> H <sub>6</sub> (against SiH <sub>4</sub> ) 100 ppm                                     |                             |                                            |                       |                      |
|                                  | SiH <sub>4</sub> 100                                                                                  |                             |                                            |                       |                      |
|                                  | B <sub>2</sub> H <sub>6</sub> (against SiH <sub>4</sub> ) 500 ppm (LL-side:2 μm) (U·2nd·LR-side:1 μm) |                             |                                            |                       |                      |
|                                  | 500 ppm→0**                                                                                           |                             |                                            |                       |                      |
|                                  | H <sub>2</sub> 200                                                                                    |                             |                                            |                       |                      |
|                                  | 2nd layer region SiH <sub>4</sub> 400                                                                 |                             |                                            |                       |                      |
| Upper layer                      | Ar 200                                                                                                | 250                         | 10                                         | 0.5                   | 15                   |
|                                  | 3rd layer region SiH <sub>4</sub> 100                                                                 |                             |                                            |                       |                      |
|                                  | NH <sub>3</sub> 30                                                                                    |                             |                                            |                       |                      |

TABLE 39

| Order of lamination (layer name) | Gases and their flow rates (SCCM)                                     | Substrate temperature (°C.) | RF discharging power (mW/cm <sup>3</sup> ) | Inner pressure (Torr) | Layer thickness (μm) |
|----------------------------------|-----------------------------------------------------------------------|-----------------------------|--------------------------------------------|-----------------------|----------------------|
| Lower layer                      | SiH <sub>4</sub> 10→100*                                              | 300                         | 10                                         | 0.4                   | 0.2                  |
|                                  | H <sub>2</sub> 5→200*                                                 |                             |                                            |                       |                      |
|                                  | AlCl <sub>3</sub> /He (S-side:0.05 μm)                                |                             |                                            |                       |                      |
|                                  | 200→40* (UL-side:0.15 μm)                                             |                             |                                            |                       |                      |
|                                  | B <sub>2</sub> H <sub>6</sub> (against SiH <sub>4</sub> ) 100 ppm     |                             |                                            |                       |                      |
|                                  | SiH <sub>4</sub> 100                                                  |                             |                                            |                       |                      |
|                                  | B <sub>2</sub> H <sub>6</sub> 200 ppm                                 |                             |                                            |                       |                      |
|                                  | H <sub>2</sub> 500                                                    |                             |                                            |                       |                      |
|                                  | 2nd layer region SiH <sub>4</sub> 300                                 |                             |                                            |                       |                      |
|                                  | H <sub>2</sub> 500                                                    |                             |                                            |                       |                      |
| Upper layer                      | 3rd layer region SiH <sub>4</sub> 100                                 | 300                         | 20                                         | 0.5                   | 20                   |
|                                  | CH <sub>4</sub> 600                                                   |                             |                                            |                       |                      |
|                                  | 4th layer region PH <sub>3</sub> (against SiH <sub>4</sub> ) 3000 ppm |                             |                                            |                       |                      |
|                                  | SiH <sub>4</sub> 40                                                   |                             |                                            |                       |                      |
|                                  | CH <sub>4</sub> 600                                                   |                             |                                            |                       |                      |
|                                  | B <sub>2</sub> H <sub>6</sub> (against SiH <sub>4</sub> ) 5000 ppm    |                             |                                            |                       |                      |

TABLE 40

| Order of lamination (layer name) | Gases of their flow rates (SCCM)                                   | Substrate temperature (°C.) | RF discharging power (mW/cm <sup>3</sup> ) | Inner pressure (Torr) | Layer thickness (μm) |
|----------------------------------|--------------------------------------------------------------------|-----------------------------|--------------------------------------------|-----------------------|----------------------|
| Lower layer                      | SiH <sub>4</sub> 50                                                | 330                         | 5                                          | 0.4                   | 0.05                 |
|                                  | H <sub>2</sub> 5→200*                                              |                             |                                            |                       |                      |
|                                  | AlCl <sub>3</sub> /He 200→20**                                     |                             |                                            |                       |                      |
|                                  | PH <sub>3</sub> (against SiH <sub>4</sub> ) 50 ppm                 |                             |                                            |                       |                      |
|                                  | SiH <sub>4</sub> 100                                               |                             |                                            |                       |                      |
|                                  | PH <sub>3</sub> 100 ppm                                            |                             |                                            |                       |                      |
|                                  | H <sub>2</sub> 100                                                 |                             |                                            |                       |                      |
|                                  | 2nd layer region SiH <sub>4</sub> 400                              |                             |                                            |                       |                      |
|                                  | SiF <sub>4</sub> 10                                                |                             |                                            |                       |                      |
|                                  | H <sub>2</sub> 800                                                 |                             |                                            |                       |                      |
| Upper layer                      | 3rd layer region SiH <sub>4</sub> 100                              | 350                         | 15                                         | 0.4                   | 5                    |
|                                  | CH <sub>4</sub> 400                                                |                             |                                            |                       |                      |
|                                  | B <sub>2</sub> H <sub>6</sub> (against SiH <sub>4</sub> ) 5000 ppm |                             |                                            |                       |                      |
|                                  | SiH <sub>4</sub> 20                                                |                             |                                            |                       |                      |
|                                  | CH <sub>4</sub> 400                                                |                             |                                            |                       |                      |
|                                  | B <sub>2</sub> H <sub>6</sub> (against SiH <sub>4</sub> ) 8000 ppm |                             |                                            |                       |                      |

TABLE 41

| Order of lamination (layer name) | Gases of their flow rates (SCCM)                          |                                                      | Substrate temperature (°C.) | RF discharging power (mW/cm <sup>3</sup> ) | Inner pressure (Torr) | Layer thickness (μm) |
|----------------------------------|-----------------------------------------------------------|------------------------------------------------------|-----------------------------|--------------------------------------------|-----------------------|----------------------|
| Lower layer                      | SiH <sub>4</sub>                                          | 50                                                   | 300                         | 1                                          | 0.3                   | 0.02                 |
|                                  | H <sub>2</sub>                                            | 10→200*                                              |                             |                                            |                       |                      |
|                                  | AlCl <sub>3</sub> /He (S-side: 0.01 μm)                   | 200→30**                                             |                             |                                            |                       |                      |
|                                  | (UL-side: 0.01 μm)                                        | 30→10**                                              |                             |                                            |                       |                      |
|                                  | B <sub>2</sub> H <sub>6</sub> (against SiH <sub>4</sub> ) | 100 ppm                                              |                             |                                            |                       |                      |
|                                  | SiH <sub>4</sub>                                          | 100                                                  |                             |                                            |                       |                      |
|                                  | B <sub>2</sub> H <sub>6</sub> (against SiH <sub>4</sub> ) | 200 ppm                                              |                             |                                            |                       |                      |
|                                  | H <sub>2</sub>                                            | 500                                                  |                             |                                            |                       |                      |
|                                  | 2nd layer region                                          | SiH <sub>4</sub> 300                                 |                             |                                            |                       |                      |
|                                  | 2nd layer region                                          | H <sub>2</sub> 200                                   |                             |                                            |                       |                      |
| Upper layer                      | 3rd layer region                                          | SiH <sub>4</sub> 50                                  | 300                         | 20                                         | 0.4                   | 5                    |
|                                  | 3rd layer region                                          | N <sub>2</sub> 500                                   |                             |                                            |                       |                      |
|                                  | 4th layer region                                          | PH <sub>3</sub> (against SiH <sub>4</sub> ) 3000 ppm |                             |                                            |                       |                      |
|                                  | 4th layer region                                          | SiH <sub>4</sub> 40                                  |                             |                                            |                       |                      |
|                                  | 4th layer region                                          | CH <sub>4</sub> 600                                  |                             |                                            |                       |                      |

TABLE 42

| Order of lamination (layer name) | Gases and their flow rates (SCCM)                         |                                      | Substrate temperature (°C.) | RF discharging power (mW/cm <sup>3</sup> ) | Inner pressure (Torr) | Layer thickness (μm) |
|----------------------------------|-----------------------------------------------------------|--------------------------------------|-----------------------------|--------------------------------------------|-----------------------|----------------------|
| Lower layer                      | SiH <sub>4</sub>                                          | 50                                   | 250                         | 5                                          | 0.4                   | 0.05                 |
|                                  | H <sub>2</sub>                                            | 5→200*                               |                             |                                            |                       |                      |
|                                  | AlCl <sub>3</sub> /He                                     | 200→20**                             |                             |                                            |                       |                      |
|                                  | B <sub>2</sub> H <sub>6</sub> (against SiH <sub>4</sub> ) | 10 ppm                               |                             |                                            |                       |                      |
|                                  | SiH <sub>4</sub>                                          | 100                                  |                             |                                            |                       |                      |
|                                  | B <sub>2</sub> H <sub>6</sub> (against SiH <sub>4</sub> ) | 500 ppm                              |                             |                                            |                       |                      |
|                                  | (LL-side: 3 μm)                                           | 500 ppm→0**                          |                             |                                            |                       |                      |
|                                  | (U·2nd·LR-side: 2 μm)                                     | 200                                  |                             |                                            |                       |                      |
|                                  | H <sub>2</sub>                                            | 1→0**                                |                             |                                            |                       |                      |
|                                  | AlCl <sub>3</sub> /He (against SiH <sub>4</sub> )         | 300                                  |                             |                                            |                       |                      |
| Upper layer                      | 2nd layer region                                          | SiH <sub>4</sub> 300                 | 250                         | 15                                         | 0.5                   | 10                   |
|                                  | 2nd layer region                                          | H <sub>2</sub> 300                   |                             |                                            |                       |                      |
|                                  | 3rd layer region                                          | SiH <sub>4</sub> 200                 |                             |                                            |                       |                      |
|                                  | 3rd layer region                                          | C <sub>2</sub> H <sub>2</sub> 10→20* |                             |                                            |                       |                      |
|                                  | 4th layer region                                          | NO 1                                 |                             |                                            |                       |                      |

TABLE 43

| Order of lamination (layer name) | Gases of their flow rates (SCCM)                          |                      | Substrate temperature (°C.) | RF discharging power (mW/cm <sup>3</sup> ) | Inner pressure (Torr) | Layer thickness (μm) |
|----------------------------------|-----------------------------------------------------------|----------------------|-----------------------------|--------------------------------------------|-----------------------|----------------------|
| Lower layer                      | H <sub>2</sub> S(against SiH <sub>4</sub> )               | 10 ppm               | 1                           | 0.4                                        | 0.02                  | 0.02                 |
|                                  | SiH <sub>4</sub>                                          | 50                   |                             |                                            |                       |                      |
|                                  | H <sub>2</sub>                                            | 5→200*               |                             |                                            |                       |                      |
|                                  | AlCl <sub>3</sub> /He (S-side: 0.01 μm)                   | 250                  |                             |                                            |                       |                      |
|                                  | (UL-side: 0.01 μm)                                        | 200→30**             |                             |                                            |                       |                      |
|                                  | B <sub>2</sub> H <sub>6</sub> (against SiH <sub>4</sub> ) | 30→10**              |                             |                                            |                       |                      |
|                                  | SiH <sub>4</sub>                                          | 100 ppm              |                             |                                            |                       |                      |
|                                  | B <sub>2</sub> H <sub>6</sub> (against SiH <sub>4</sub> ) | 100                  |                             |                                            |                       |                      |
|                                  | (LL-side: 2 μm)                                           | 500 ppm              |                             |                                            |                       |                      |
|                                  | (U·2nd·LR-side: 1 μm)                                     | 500 ppm→0**          |                             |                                            |                       |                      |
| Upper layer                      | 2nd layer region                                          | H <sub>2</sub> 200   | 300                         | 20                                         | 0.5                   | 5                    |
|                                  | 2nd layer region                                          | SiH <sub>4</sub> 300 |                             |                                            |                       |                      |
|                                  | 3rd layer region                                          | H <sub>2</sub> 300   |                             |                                            |                       |                      |
|                                  | 3rd layer region                                          | SiH <sub>4</sub> 100 |                             |                                            |                       |                      |
|                                  | 4th layer region                                          | CH <sub>4</sub> 100  |                             |                                            |                       |                      |
| 4th layer                        | SiH <sub>4</sub>                                          | 50                   | 300                         | 15                                         | 0.4                   | 20                   |
|                                  | CH <sub>4</sub>                                           | 600                  |                             |                                            |                       |                      |

TABLE 43-continued

| Order of lamination (layer name) | Gases of their flow rates (SCCM) | Substrate temperature (°C.) | RF discharging power (mW/cm <sup>3</sup> ) | Inner pressure (Torr) | Layer thickness (μm) |
|----------------------------------|----------------------------------|-----------------------------|--------------------------------------------|-----------------------|----------------------|
| region                           |                                  |                             |                                            |                       |                      |

TABLE 44

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 10→100*                                          | 300                         | 5                                          | 0.4                   | 0.2                  |
|                                  | H <sub>2</sub> 5→200*                                             |                             |                                            |                       |                      |
|                                  | AlCl <sub>3</sub> /He (S-side: 0.05 μm)                           |                             |                                            |                       |                      |
|                                  | 200→40** (UL-side: 0.15 μm)                                       |                             |                                            |                       |                      |
|                                  | 40→10**                                                           |                             |                                            |                       |                      |
|                                  | B <sub>2</sub> H <sub>6</sub> (against SiH <sub>4</sub> ) 50 ppm  |                             |                                            |                       |                      |
|                                  | SiH <sub>4</sub> 100                                              |                             |                                            |                       |                      |
|                                  | B <sub>2</sub> H <sub>4</sub> (against SiH <sub>4</sub> ) 200 ppm |                             |                                            |                       |                      |
|                                  | H <sub>2</sub> 500                                                |                             |                                            |                       |                      |
|                                  | SiH <sub>4</sub> 100                                              |                             |                                            |                       |                      |
| Upper layer                      | H <sub>2</sub> 300                                                |                             |                                            |                       |                      |
|                                  | 1st layer region 3rd layer region 4th layer region                | 300                         | 5                                          | 0.4                   | 3                    |
|                                  | SiH <sub>4</sub> 300                                              |                             |                                            |                       |                      |
|                                  | NH <sub>3</sub> 50                                                |                             |                                            |                       |                      |
|                                  | SiH <sub>4</sub> 100                                              |                             |                                            |                       |                      |
| layer region                     | NH <sub>3</sub> 50                                                | 300                         | 15                                         | 0.4                   | 25                   |
|                                  | SiH <sub>4</sub> 100                                              | 300                         | 10                                         | 0.4                   | 0.3                  |

TABLE 45

| Order of lamination (layer name) | Gases and their flow rates (SCCM)                                                                   | Substrate temperature (°C.) | RF discharging power (mW/cm <sup>3</sup> ) | Inner pressure (Torr) | Layer thickness (μm) |
|----------------------------------|-----------------------------------------------------------------------------------------------------|-----------------------------|--------------------------------------------|-----------------------|----------------------|
| Lower layer                      | SiH <sub>4</sub> 10→100*                                                                            | 250                         | 5                                          | 0.4                   | 0.2                  |
|                                  | H <sub>2</sub> 5→200*                                                                               |                             |                                            |                       |                      |
|                                  | AlCl <sub>3</sub> /He (S-side: 0.05 μm)                                                             |                             |                                            |                       |                      |
|                                  | 200→40** (UL-side: 0.15 μm)                                                                         |                             |                                            |                       |                      |
|                                  | 40→10**                                                                                             |                             |                                            |                       |                      |
|                                  | B <sub>2</sub> H <sub>6</sub> (against SiH <sub>4</sub> ) 100 ppm                                   |                             |                                            |                       |                      |
|                                  | SiH <sub>4</sub> 100                                                                                |                             |                                            |                       |                      |
|                                  | B <sub>2</sub> H <sub>6</sub> (against SiH <sub>4</sub> ) (LL-side: 2 μm) (U · 2nd · LR-side: 1 μm) |                             |                                            |                       |                      |
|                                  | 500 ppm→0**                                                                                         |                             |                                            |                       |                      |
|                                  | H <sub>2</sub> 200                                                                                  |                             |                                            |                       |                      |
| Upper layer                      | SiH <sub>4</sub> 100                                                                                |                             |                                            |                       |                      |
|                                  | SiF <sub>4</sub> 5                                                                                  | 300                         | 3                                          | 0.5                   | 3                    |
|                                  | H <sub>2</sub> 200                                                                                  |                             |                                            |                       |                      |
|                                  | SiH <sub>4</sub> 100                                                                                |                             |                                            |                       |                      |
|                                  | CH <sub>4</sub> 100                                                                                 | 300                         | 15                                         | 0.4                   | 30                   |
|                                  | PH <sub>3</sub> (against SiH <sub>4</sub> ) 50 ppm                                                  |                             |                                            |                       |                      |
|                                  | SiH <sub>4</sub> 50                                                                                 |                             |                                            |                       |                      |
|                                  | CH <sub>4</sub> 600                                                                                 | 300                         | 10                                         | 0.4                   | 0.5                  |

TABLE 46

| Order of lamination (layer name) | Gases and their flow rates (SCCM)                                                     | Substrate temperature (°C.) | RF discharging power (mW/cm <sup>3</sup> ) | Inner pressure (Torr) | Layer thickness (μm) |
|----------------------------------|---------------------------------------------------------------------------------------|-----------------------------|--------------------------------------------|-----------------------|----------------------|
| Lower layer                      | H <sub>2</sub> S (against SiH <sub>4</sub> ) 3 ppm                                    | 250                         | 5                                          | 0.4                   | 0.05                 |
|                                  | SiH <sub>4</sub> 50                                                                   |                             |                                            |                       |                      |
|                                  | H <sub>2</sub> 5→200*                                                                 |                             |                                            |                       |                      |
|                                  | AlCl <sub>3</sub> /He 200→20**                                                        |                             |                                            |                       |                      |
|                                  | PH <sub>3</sub> (against SiH <sub>4</sub> ) 100 ppm                                   |                             |                                            |                       |                      |
|                                  | SiH <sub>4</sub> 40                                                                   |                             |                                            |                       |                      |
|                                  | PH <sub>3</sub> (against SiH <sub>4</sub> ) (LL-side: 2 μm) (U · 2nd · LR-side: 1 μm) |                             |                                            |                       |                      |
|                                  | 250 ppm→0**                                                                           |                             |                                            |                       |                      |
|                                  | H <sub>2</sub> 40                                                                     |                             |                                            |                       |                      |
|                                  | Si <sub>2</sub> H <sub>6</sub> 200                                                    |                             |                                            |                       |                      |
| Upper layer                      | SiH <sub>4</sub> 40                                                                   |                             |                                            |                       |                      |
|                                  | PH <sub>3</sub> (against SiH <sub>4</sub> ) 250 ppm→0**                               |                             |                                            |                       |                      |
| 2nd                              | SiH <sub>4</sub> 40                                                                   |                             |                                            |                       |                      |

TABLE 46-continued

| Order of lamination (layer name) | Gases and their flow rates (SCCM)                                                   | Substrate temperature (°C.) | RF discharging power (mW/cm <sup>3</sup> ) | Inner pressure (Torr) | Layer thickness (μm) |
|----------------------------------|-------------------------------------------------------------------------------------|-----------------------------|--------------------------------------------|-----------------------|----------------------|
| layer region                     | H <sub>2</sub> 200                                                                  | 300                         | 10                                         | 0.5                   | 10                   |
| 3rd layer region                 | SiH <sub>4</sub> 300                                                                |                             |                                            |                       |                      |
|                                  | C <sub>2</sub> H <sub>2</sub> 50                                                    |                             |                                            |                       |                      |
|                                  | B <sub>2</sub> H <sub>6</sub> (against SiH <sub>4</sub> ) (U · 2nd · LR-side: 1 μm) | 330                         | 20                                         | 0.4                   | 30                   |
|                                  | 0→100 ppm*                                                                          |                             |                                            |                       |                      |
|                                  | (U · 3rd · LR-side 29 μm) 100 ppm                                                   |                             |                                            |                       |                      |
| 4th layer region                 | SiH <sub>4</sub> 200                                                                | 330                         | 10                                         | 0.4                   | 1                    |
|                                  | C <sub>2</sub> H <sub>2</sub> 200                                                   |                             |                                            |                       |                      |

TABLE 47

| Order of lamination (layer name) | Gases and their flow rates (SCCM)                                                                                                                                                                                                                                                                                                                                                                                                                                                                                       | Substrate temperature (°C.) | RF discharging power (mW/cm <sup>3</sup> ) | Inner pressure (Torr) | Layer thickness (μm) |
|----------------------------------|-------------------------------------------------------------------------------------------------------------------------------------------------------------------------------------------------------------------------------------------------------------------------------------------------------------------------------------------------------------------------------------------------------------------------------------------------------------------------------------------------------------------------|-----------------------------|--------------------------------------------|-----------------------|----------------------|
| Lower layer                      | SiH <sub>4</sub> 10→100*<br>H <sub>2</sub> 5→200*                                                                                                                                                                                                                                                                                                                                                                                                                                                                       | 250                         | 5                                          | 0.4                   | 0.2                  |
|                                  | AlCl <sub>3</sub> /He (S-side:0.05 μm) 200→40**<br>(UL-side:0.15 μm) 40→10**                                                                                                                                                                                                                                                                                                                                                                                                                                            |                             |                                            |                       |                      |
| Upper layer                      | 1st layer region B <sub>2</sub> H <sub>6</sub> (against SiH <sub>4</sub> ) 50 ppm<br>SiH <sub>4</sub> 100<br>B <sub>2</sub> H <sub>6</sub> (against SiH <sub>4</sub> ) 200 ppm<br>H <sub>2</sub> 500<br>2nd layer region SiH <sub>4</sub> 100<br>H <sub>2</sub> 300<br>3rd layer region SiH <sub>4</sub> 300<br>NH <sub>3</sub> 30→50*<br>PH <sub>3</sub> (against SiH <sub>4</sub> ) 50 ppm<br>4th layer region SiH <sub>4</sub> 100<br>NH <sub>3</sub> 80→100*<br>PH <sub>3</sub> (against SiH <sub>4</sub> ) 500 ppm | 300                         | 8                                          | 0.3                   | 3                    |
|                                  |                                                                                                                                                                                                                                                                                                                                                                                                                                                                                                                         |                             | 5                                          | 0.2                   | 8                    |
|                                  |                                                                                                                                                                                                                                                                                                                                                                                                                                                                                                                         | 300                         | 15                                         | 0.4                   | 25                   |
|                                  |                                                                                                                                                                                                                                                                                                                                                                                                                                                                                                                         | 300                         | 5                                          | 0.4                   | 0.7                  |

TABLE 48

| Order of lamination (layer name) | Gases and their flow rates (SCCM)                                                                                                                                                                                                                                                                                                                        | Substrate temperature (°C.) | RF discharging power (mW/cm <sup>3</sup> ) | Inner pressure (Torr) | Layer thickness (μm) |
|----------------------------------|----------------------------------------------------------------------------------------------------------------------------------------------------------------------------------------------------------------------------------------------------------------------------------------------------------------------------------------------------------|-----------------------------|--------------------------------------------|-----------------------|----------------------|
| Lower layer                      | SiH <sub>4</sub> 50<br>H <sub>2</sub> 5→200*                                                                                                                                                                                                                                                                                                             | 250                         | 1                                          | 0.4                   | 0.02                 |
|                                  | AlCl <sub>3</sub> /He (S-side:0.01 μm) 200→30**<br>(UL-side:0.01 μm) 30→10**                                                                                                                                                                                                                                                                             |                             |                                            |                       |                      |
| Upper layer                      | 1st layer region PH <sub>3</sub> (against SiH <sub>4</sub> ) 30 ppm<br>SiH <sub>4</sub> 100<br>H <sub>2</sub> 100 ppm<br>2nd layer region SiH <sub>4</sub> 300<br>H <sub>2</sub> 500<br>3rd layer region SiH <sub>4</sub> 100<br>GeH <sub>4</sub> 10→50*<br>H <sub>2</sub> 300<br>4th layer region SiH <sub>4</sub> 100→40**<br>CH <sub>4</sub> 100→600* | 300                         | 8                                          | 0.4                   | 3                    |
|                                  |                                                                                                                                                                                                                                                                                                                                                          |                             | 20                                         | 0.5                   | 20                   |
|                                  |                                                                                                                                                                                                                                                                                                                                                          | 300                         | 5                                          | 0.4                   | 1                    |
|                                  |                                                                                                                                                                                                                                                                                                                                                          | 300                         | 10                                         | 0.4                   | 1                    |

TABLE 49

| Order of lamination (layer name) | Gases and their flow rates (SCCM)            | Substrate temperature (°C.) | RF discharging power (mW/cm <sup>3</sup> ) | Inner pressure (Torr) | Layer thickness (μm) |
|----------------------------------|----------------------------------------------|-----------------------------|--------------------------------------------|-----------------------|----------------------|
| Lower layer                      | SiH <sub>4</sub> 50<br>H <sub>2</sub> 5→200* | 300                         | 1                                          | 0.3                   | 0.02                 |
|                                  | AlCl <sub>3</sub> /He (S-side:0.01 μm)       |                             |                                            |                       |                      |

TABLE 49-continued

| Order of lamination (layer name) | Gases and their flow rates (SCCM)                                    | Substrate temperature (°C.) | RF discharging power (mW/cm <sup>3</sup> ) | Inner pressure (Torr) | Layer thickness (μm) |
|----------------------------------|----------------------------------------------------------------------|-----------------------------|--------------------------------------------|-----------------------|----------------------|
| Upper layer                      | 200→30**<br>(UL-side:0.01 μm)                                        |                             |                                            |                       |                      |
|                                  | 30→10**<br>B <sub>2</sub> H <sub>6</sub> (against SiH <sub>4</sub> ) | 100 ppm                     |                                            |                       |                      |
|                                  | SiH <sub>4</sub>                                                     | 100                         |                                            |                       |                      |
|                                  | B <sub>2</sub> H <sub>6</sub> (against SiH <sub>4</sub> )            | 200 ppm                     | 300                                        | 8                     | 0.4                  |
|                                  | H <sub>2</sub>                                                       | 500                         |                                            |                       |                      |
|                                  | SiH <sub>4</sub>                                                     | 300                         |                                            |                       |                      |
|                                  | H <sub>2</sub>                                                       | 400                         | 300                                        | 15                    | 0.5                  |
|                                  | SiH <sub>4</sub>                                                     | 50                          |                                            |                       |                      |
|                                  | CH <sub>4</sub>                                                      | 500                         | 300                                        | 10                    | 0.4                  |
|                                  |                                                                      |                             |                                            |                       | 0.5                  |

TABLE 50

| Order of lamination (layer name) | Gases and their flow rates (SCCM)                                    | Substrate temperature (°C.) | RF discharging power (mW/cm <sup>3</sup> ) | Inner pressure (Torr) | Layer thickness (μm) |
|----------------------------------|----------------------------------------------------------------------|-----------------------------|--------------------------------------------|-----------------------|----------------------|
| Upper layer                      | SiH <sub>4</sub>                                                     | 50                          |                                            |                       |                      |
|                                  | H <sub>2</sub>                                                       | 5→200*                      |                                            |                       |                      |
|                                  | AlCl <sub>3</sub> /He<br>(S-side:0.01 μm)                            |                             | 300                                        | 0.7                   | 0.3                  |
|                                  | 200→30**<br>(UL-side:0.01 μm)                                        |                             |                                            |                       |                      |
|                                  | 30→10**<br>B <sub>2</sub> H <sub>6</sub> (against SiH <sub>4</sub> ) | 50 ppm                      |                                            |                       |                      |
|                                  | SiH <sub>4</sub>                                                     | 100                         |                                            |                       |                      |
|                                  | B <sub>2</sub> H <sub>6</sub> (against SiH <sub>4</sub> )            | 200 ppm                     | 300                                        | 7                     | 0.3                  |
|                                  | H <sub>2</sub>                                                       | 500                         |                                            |                       |                      |
|                                  | SiH <sub>4</sub>                                                     | 200                         |                                            |                       |                      |
|                                  | H <sub>2</sub>                                                       | 400                         | 300                                        | 12                    | 0.4                  |
|                                  | SiH <sub>4</sub>                                                     | 40                          |                                            |                       |                      |
|                                  | CH <sub>4</sub>                                                      | 400                         | 300                                        | 7                     | 0.3                  |
|                                  |                                                                      |                             |                                            |                       | 0.5                  |

TABLE 51

| Order of lamination (layer name) | Gases and their flow rates (SCCM)                                   | Substrate temperature (°C.) | RF discharging power (mW/cm <sup>3</sup> ) | Inner pressure (Torr) | Layer thickness (μm) |
|----------------------------------|---------------------------------------------------------------------|-----------------------------|--------------------------------------------|-----------------------|----------------------|
| Upper layer                      | SiH <sub>4</sub>                                                    | 25                          |                                            |                       |                      |
|                                  | H <sub>2</sub>                                                      | 5→100*                      |                                            |                       |                      |
|                                  | AlCl <sub>3</sub> /He<br>(S-side:0.01 μm)                           |                             | 300                                        | 0.5                   | 0.2                  |
|                                  | 100→15**<br>(UL-side:0.01 μm)                                       |                             |                                            |                       |                      |
|                                  | 15→5**<br>B <sub>2</sub> H <sub>6</sub> (against SiH <sub>4</sub> ) | 30 ppm                      |                                            |                       |                      |
|                                  | SiH <sub>4</sub>                                                    | 100                         |                                            |                       |                      |
|                                  | B <sub>2</sub> H <sub>6</sub> (against SiH <sub>4</sub> )           | 200 ppm                     | 300                                        | 6                     | 0.2                  |
|                                  | H <sub>2</sub>                                                      | 500                         |                                            |                       |                      |
|                                  | SiH <sub>4</sub>                                                    | 150                         |                                            |                       |                      |
|                                  | H <sub>2</sub>                                                      | 300                         | 300                                        | 10                    | 0.4                  |
|                                  | SiH <sub>4</sub>                                                    | 30                          |                                            |                       |                      |
|                                  | CH <sub>4</sub>                                                     | 300                         | 300                                        | 5                     | 0.3                  |
|                                  |                                                                     |                             |                                            |                       | 0.5                  |

TABLE 52

| Order of lamination (layer name) | Gases and their flow rates (SCCM)                                   | Substrate temperature (°C.) | RF discharging power (mW/cm <sup>3</sup> ) | Inner pressure (Torr) | Layer thickness (μm) |
|----------------------------------|---------------------------------------------------------------------|-----------------------------|--------------------------------------------|-----------------------|----------------------|
| Upper layer                      | SiH <sub>4</sub>                                                    | 20                          |                                            |                       |                      |
|                                  | H <sub>2</sub>                                                      | 5→100*                      |                                            |                       |                      |
|                                  | AlCl <sub>3</sub> /He<br>(S-side:0.01 μm)                           |                             | 300                                        | 0.3                   | 0.2                  |
|                                  | 80→15**<br>(UL-side:0.01 μm)                                        |                             |                                            |                       |                      |
|                                  | 15→5**<br>B <sub>2</sub> H <sub>6</sub> (against SiH <sub>4</sub> ) | 30 ppm                      |                                            |                       |                      |
|                                  | SiH <sub>4</sub>                                                    | 100                         |                                            |                       |                      |
|                                  | B <sub>2</sub> H <sub>6</sub> (against SiH <sub>4</sub> )           |                             |                                            |                       |                      |
|                                  |                                                                     |                             |                                            |                       |                      |
|                                  |                                                                     |                             |                                            |                       |                      |

TABLE 52-continued

| Order of lamination (layer name) |                  | Gases and their flow rates (SCCM)                                           | Substrate temperature (°C.) | RF discharging power (mW/cm <sup>3</sup> ) | Inner pressure (Torr) | Layer thickness (μm) |
|----------------------------------|------------------|-----------------------------------------------------------------------------|-----------------------------|--------------------------------------------|-----------------------|----------------------|
| layer                            | layer region     | B <sub>2</sub> H <sub>6</sub> (against SiH <sub>4</sub> )<br>H <sub>2</sub> | 200 ppm<br>500              | 300                                        | 5                     | 0.2                  |
|                                  | 2nd layer region | SiH <sub>4</sub>                                                            | 100                         |                                            |                       |                      |
|                                  | layer region     | H <sub>2</sub>                                                              | 300                         | 300                                        | 6                     | 0.3                  |
|                                  | 3rd layer region | SiH <sub>4</sub>                                                            | 20                          | 300                                        | 3                     | 0.2                  |
|                                  | layer region     | CH <sub>4</sub>                                                             | 200                         |                                            |                       | 0.5                  |
|                                  |                  | SiH <sub>4</sub>                                                            | 100                         |                                            |                       |                      |

TABLE 53

| Order of lamination (layer name) |                  | Gases and their flow rates (SCCM)                                           | Substrate temperature (°C.) | RF discharging power (mW/cm <sup>3</sup> ) | Inner pressure (Torr) | Layer thickness (μm) |
|----------------------------------|------------------|-----------------------------------------------------------------------------|-----------------------------|--------------------------------------------|-----------------------|----------------------|
| Lower layer                      |                  | SiH <sub>4</sub>                                                            | 50                          |                                            |                       |                      |
|                                  |                  | H <sub>2</sub>                                                              | 5→200*                      | 500                                        | 5                     | 0.4                  |
|                                  |                  | AlCl <sub>3</sub> /He                                                       | 200→20**                    |                                            |                       |                      |
|                                  |                  | B <sub>2</sub> H <sub>6</sub> (against SiH <sub>4</sub> )                   | 100 ppm                     |                                            |                       |                      |
| Upper layer                      | 1st layer region | SiH <sub>4</sub>                                                            | 100                         |                                            |                       |                      |
|                                  |                  | B <sub>2</sub> H <sub>6</sub> (against SiH <sub>4</sub> )<br>(LL-side:2 μm) | 500 ppm                     | 500                                        | 7                     | 0.4                  |
|                                  |                  | (U·2nd·LR-side:1 μm)                                                        | 500 ppm→0**                 |                                            |                       | 3                    |
|                                  | 2nd layer region | H <sub>2</sub>                                                              | 200                         |                                            |                       |                      |
|                                  |                  | SiH <sub>4</sub>                                                            | 300                         |                                            |                       |                      |
|                                  |                  | H <sub>2</sub>                                                              | 1500                        | 500                                        | 30                    | 0.5                  |
|                                  | 3rd layer region | SiH <sub>4</sub>                                                            | 200                         |                                            |                       |                      |
|                                  |                  | C <sub>2</sub> H <sub>2</sub>                                               | 10→20*                      | 500                                        | 30                    | 0.4                  |
|                                  |                  | NO                                                                          | 1                           |                                            |                       | 20                   |

TABLE 54

| Order of lamination (layer name) |                  | Gases and their flow rates (SCCM)                         | Substrate temperature (°C.) | μW discharging power (mW/cm <sup>3</sup> ) | Inner pressure (Torr) | Layer thickness (μm) |
|----------------------------------|------------------|-----------------------------------------------------------|-----------------------------|--------------------------------------------|-----------------------|----------------------|
| Lower layer                      |                  | H <sub>2</sub> S(against SiH <sub>4</sub> )               | 3 ppm                       |                                            |                       |                      |
|                                  |                  | SiH <sub>4</sub>                                          | 150                         |                                            |                       |                      |
|                                  |                  | H <sub>2</sub>                                            | 20→500*                     |                                            |                       |                      |
|                                  |                  | AlCl <sub>3</sub> /He<br>(S-side:0.01 μm)                 |                             | 250                                        | 0.5                   | 0.6                  |
|                                  |                  |                                                           | 80→50**                     |                                            |                       |                      |
| Upper layer                      | 1st layer region | B <sub>2</sub> H <sub>6</sub> (against SiH <sub>4</sub> ) | 50 ppm                      |                                            |                       |                      |
|                                  |                  | SiH <sub>4</sub>                                          | 100                         |                                            |                       |                      |
|                                  |                  | B <sub>2</sub> H <sub>6</sub> (against SiH <sub>4</sub> ) | 200 ppm                     | 250                                        | 0.5                   | 0.5                  |
|                                  |                  | H <sub>2</sub>                                            | 500                         | 250                                        | 0.5                   | 700                  |
|                                  | 2nd layer region | SiF <sub>4</sub>                                          | 30                          |                                            |                       |                      |
|                                  |                  | H <sub>2</sub>                                            | 500                         |                                            |                       |                      |
|                                  | 3rd layer region | SiH <sub>4</sub>                                          | 150                         |                                            |                       |                      |
|                                  |                  | CH <sub>4</sub>                                           | 500                         | 250                                        | 0.5                   | 1                    |
|                                  |                  |                                                           |                             |                                            |                       |                      |

TABLE 55

| Order of lamination (layer name) |                  | Gases and their flow rates (SCCM)                                           | Substrate temperature (°C.) | RF discharging power (mW/cm <sup>3</sup> ) | Inner pressure (Torr) | Layer thickness (μm) |
|----------------------------------|------------------|-----------------------------------------------------------------------------|-----------------------------|--------------------------------------------|-----------------------|----------------------|
| Lower layer                      |                  | SiH <sub>4</sub>                                                            | 50                          |                                            |                       |                      |
|                                  |                  | H <sub>2</sub>                                                              | 5→200*                      | 250                                        | 5                     | 0.4                  |
|                                  |                  | AlCl <sub>3</sub> /He                                                       | 200→20**                    |                                            |                       |                      |
|                                  |                  | B <sub>2</sub> H <sub>6</sub> (against SiH <sub>4</sub> )                   | 100 ppm                     |                                            |                       |                      |
| Upper layer                      | 1st layer region | SiH <sub>4</sub>                                                            | 100                         |                                            |                       |                      |
|                                  |                  | B <sub>2</sub> H <sub>6</sub> (against SiH <sub>4</sub> )<br>(LL-side:3 μm) | 500 ppm                     |                                            |                       |                      |
|                                  |                  | (U·2nd·LR-side:2 μm)                                                        | 250                         | 10                                         | 0.4                   | 5                    |
|                                  |                  |                                                                             | 500 ppm→0**                 |                                            |                       |                      |
|                                  | 2nd layer region | H <sub>2</sub>                                                              | 200                         |                                            |                       |                      |
|                                  |                  | AlCl <sub>3</sub> /He<br>(against SiH <sub>4</sub> )1→0**                   |                             |                                            |                       |                      |
|                                  | 3rd layer region | SiH <sub>4</sub>                                                            | 200                         | 250                                        | 15                    | 0.4                  |
|                                  |                  | C <sub>2</sub> H <sub>2</sub>                                               | 10→20*                      |                                            |                       | 20                   |
|                                  |                  | NO                                                                          | 1                           |                                            |                       |                      |
|                                  |                  | SiH <sub>4</sub>                                                            | 300                         |                                            |                       |                      |

TABLE 55-continued

| Order of lamination (layer name) | Gases and their flow rates (SCCM) | Substrate temperature (°C.) | RF discharging power (mW/cm <sup>3</sup> ) | Inner pressure (Torr) | Layer thickness (μm) |
|----------------------------------|-----------------------------------|-----------------------------|--------------------------------------------|-----------------------|----------------------|
| layer region                     | H <sub>2</sub> 300                | 250                         | 15                                         | 0.5                   | 10                   |

TABLE 56

| Order of lamination (layer name) | Gases and their flow rates (SCCM)                                                                                        | Substrate temperature (°C.) | RF discharging power (mW/cm <sup>3</sup> ) | Inner pressure (Torr) | Layer thickness (μm) |
|----------------------------------|--------------------------------------------------------------------------------------------------------------------------|-----------------------------|--------------------------------------------|-----------------------|----------------------|
| Lower layer                      | SiH <sub>4</sub> 50<br>H <sub>2</sub> 5→200*                                                                             | 250                         | 1                                          | 0.4                   | 0.02                 |
|                                  | AlCl <sub>3</sub> /He (S-side:0.01 μm) 200→30**<br>(UL-side:0.01 μm) 30→10**                                             |                             |                                            |                       |                      |
| Upper layer                      | B <sub>2</sub> H <sub>6</sub> (against SiH <sub>4</sub> ) 50 ppm<br>SiH <sub>4</sub> 100                                 |                             |                                            |                       |                      |
| 1st layer region                 | B <sub>2</sub> H <sub>6</sub> (against SiH <sub>4</sub> ) 500 ppm<br>(LL-side:2 μm) (U · 2nd · LR-side:1 μm) 500 ppm→0** | 250                         | 10                                         | 0.4                   | 10                   |
| 2nd layer region                 | H <sub>2</sub> 200<br>SiH <sub>4</sub> 100                                                                               | 300                         | 15                                         | 0.4                   | 20                   |
| 3rd layer region                 | CH <sub>4</sub> 100                                                                                                      | 300                         | 20                                         | 0.5                   | 5                    |
| 4th layer region                 | SiH <sub>4</sub> 300<br>H <sub>2</sub> 300                                                                               | 300                         | 10                                         | 0.4                   | 0.5                  |

TABLE 57

| Order of lamination (layer name) | Gases and their flow rates (SCCM)                                                                                                                                                                    | Substrate temperature (°C.) | RF discharging power (mW/cm <sup>3</sup> ) | Inner pressure (Torr) | Layer thickness (μm) |
|----------------------------------|------------------------------------------------------------------------------------------------------------------------------------------------------------------------------------------------------|-----------------------------|--------------------------------------------|-----------------------|----------------------|
| Lower layer                      | SiH <sub>4</sub> 10→100*<br>H <sub>2</sub> 5→200*                                                                                                                                                    | 300                         | 5                                          | 0.4                   | 0.2                  |
|                                  | AlCl <sub>3</sub> /He (S-side: 0.05 μm) 200→40**<br>(UL-side: 0.15 μm) 40→10**                                                                                                                       |                             |                                            |                       |                      |
| Upper layer                      | B <sub>2</sub> H <sub>6</sub> (against SiH <sub>4</sub> ) 30 ppm<br>SiH <sub>4</sub> 100<br>1st layer region B <sub>2</sub> H <sub>6</sub> (against SiH <sub>4</sub> ) 200 ppm<br>H <sub>2</sub> 500 | 300                         | 5                                          | 0.4                   | 3                    |
| 2nd layer region                 | SiH <sub>4</sub> 300                                                                                                                                                                                 | 300                         | 15                                         | 0.4                   | 25                   |
| 3rd layer region                 | NH <sub>3</sub> 50                                                                                                                                                                                   | 300                         | 5                                          | 0.2                   | 8                    |
| 4th layer region                 | SiH <sub>4</sub> 100<br>NH <sub>3</sub> 50                                                                                                                                                           | 300                         | 10                                         | 0.4                   | 0.3                  |

TABLE 58

| Order of lamination (layer name) | Gases and their flow rates (SCCM)                                                                                                                       | Substrate temperature (°C.) | RF discharging power (mW/cm <sup>3</sup> ) | Inner pressure (Torr) | Layer thickness (μm) |
|----------------------------------|---------------------------------------------------------------------------------------------------------------------------------------------------------|-----------------------------|--------------------------------------------|-----------------------|----------------------|
| Lower layer                      | SiH <sub>4</sub> 10→100*<br>H <sub>2</sub> 5→200*                                                                                                       | 250                         | 5                                          | 0.4                   | 0.2                  |
|                                  | AlCl <sub>3</sub> /He (S-side: 0.05 μm) 200→40**<br>(UL-side: 0.15 μm) 40→10**                                                                          |                             |                                            |                       |                      |
| 1st layer region                 | PH <sub>3</sub> (against SiH <sub>4</sub> ) 20 ppm<br>SiH <sub>4</sub> 100<br>PH <sub>3</sub> (against SiH <sub>4</sub> ) 100 ppm<br>H <sub>2</sub> 100 | 250                         | 8                                          | 0.4                   | 3                    |

TABLE 58-continued

| Order of lamination (layer name) | Gases and their flow rates (SCCM) |                                             | Substrate temperature (°C.) | RF discharging power (mW/cm <sup>3</sup> ) | Inner pressure (Torr) | Layer thickness (μm) |
|----------------------------------|-----------------------------------|---------------------------------------------|-----------------------------|--------------------------------------------|-----------------------|----------------------|
| Upper layer                      | 2nd layer                         | SiH <sub>4</sub>                            | 100                         |                                            |                       |                      |
|                                  |                                   | CH <sub>4</sub>                             | 100                         |                                            |                       |                      |
|                                  | region                            | PH <sub>3</sub> (against SiH <sub>4</sub> ) | 50 ppm                      |                                            |                       |                      |
|                                  | 3rd layer                         | SiH <sub>4</sub>                            | 100                         |                                            |                       |                      |
|                                  | region                            | SiF <sub>4</sub>                            | 5                           |                                            |                       |                      |
|                                  | 4th layer                         | H <sub>2</sub>                              | 200                         |                                            |                       |                      |
| region                           |                                   | SiH <sub>4</sub>                            | 50                          |                                            |                       |                      |
|                                  |                                   | CH <sub>4</sub>                             | 600                         |                                            |                       |                      |
|                                  |                                   |                                             | 300                         | 10                                         | 0.4                   | 0.5                  |

TABLE 59

| Order of lamination (layer name) | Gases and their flow rates (SCCM)                         |                                                                                                           | Substrate temperature (°C.) | RF discharging power (mW/cm <sup>3</sup> ) | Inner pressure (Torr) | Layer thickness (μm) |
|----------------------------------|-----------------------------------------------------------|-----------------------------------------------------------------------------------------------------------|-----------------------------|--------------------------------------------|-----------------------|----------------------|
| Lower layer                      | SiH <sub>4</sub>                                          | 50                                                                                                        |                             |                                            |                       |                      |
|                                  | H <sub>2</sub>                                            | 5→200*                                                                                                    |                             |                                            |                       |                      |
|                                  | AlCl <sub>3</sub> /He                                     | 200→20**                                                                                                  |                             |                                            |                       |                      |
|                                  | B <sub>2</sub> H <sub>6</sub> (against SiH <sub>4</sub> ) | 100 ppm                                                                                                   |                             |                                            |                       |                      |
|                                  | SiH <sub>4</sub>                                          | 100                                                                                                       |                             |                                            |                       |                      |
|                                  | 1st layer region                                          | B <sub>2</sub> H <sub>6</sub> (against SiH <sub>4</sub> )<br>(LL-side: 2 μm)<br>(U · 2nd · LR-side: 1 μm) | 500 ppm                     | 250                                        | 8                     | 0.4                  |
| Upper layer                      | 2nd layer region                                          | H <sub>2</sub>                                                                                            | 200                         |                                            |                       |                      |
|                                  |                                                           | SiH <sub>4</sub>                                                                                          | 300                         |                                            |                       |                      |
|                                  |                                                           | C <sub>2</sub> H <sub>2</sub>                                                                             | 50                          |                                            |                       |                      |
|                                  |                                                           | B <sub>2</sub> H <sub>6</sub> (against SiH <sub>4</sub> )<br>(U · 1st · LR-side: 1 μm)                    | 0→100 ppm*                  | 330                                        | 20                    | 0.4                  |
|                                  |                                                           | (U · 3rd · LR-side: 29 μm)                                                                                | 100 ppm                     |                                            |                       |                      |
|                                  | 3rd layer region                                          | Si <sub>2</sub> H <sub>6</sub>                                                                            | 200                         |                                            |                       |                      |
| 4th layer region                 |                                                           | H <sub>2</sub>                                                                                            | 200                         | 300                                        | 10                    | 0.5                  |
|                                  |                                                           | SiH <sub>4</sub>                                                                                          | 200                         |                                            |                       |                      |
|                                  |                                                           | C <sub>2</sub> H <sub>2</sub>                                                                             | 200                         | 330                                        | 10                    | 0.4                  |

TABLE 60

| Order of lamination (layer name) | Gases and their flow rates (SCCM)                                                           |                  | Substrate temperature (°C.) | RF discharging power (mW/cm <sup>3</sup> ) | Inner pressure (Torr) | Layer thickness (μm) |
|----------------------------------|---------------------------------------------------------------------------------------------|------------------|-----------------------------|--------------------------------------------|-----------------------|----------------------|
| Lower layer                      | SiH <sub>4</sub>                                                                            | 10→100*          |                             |                                            |                       |                      |
|                                  | H <sub>2</sub>                                                                              | 5→200*           |                             |                                            |                       |                      |
|                                  | AlCl <sub>3</sub> /He<br>(S-side: 0.05 μm)                                                  | 200→40**         | 250                         | 5                                          | 0.4                   | 0.2                  |
|                                  | (UL-side: 0.15 μm)                                                                          | 40→10**          |                             |                                            |                       |                      |
|                                  | PH <sub>3</sub> (against SiH <sub>4</sub> )                                                 | 50 ppm           |                             |                                            |                       |                      |
|                                  | SiH <sub>4</sub>                                                                            | 40               |                             |                                            |                       |                      |
| 1st layer region                 | PH <sub>3</sub> (against SiH <sub>4</sub> )<br>(LL-side: 2 μm)<br>(U · 2nd · LR-side: 1 μm) | 250 ppm          | 250                         | 8                                          | 0.4                   | 3                    |
|                                  |                                                                                             | 250 ppm→0**      |                             |                                            |                       |                      |
|                                  | H <sub>2</sub>                                                                              | 40               |                             |                                            |                       |                      |
|                                  | SiH <sub>4</sub>                                                                            | 300              |                             |                                            |                       |                      |
|                                  | NH <sub>3</sub>                                                                             | 30→50*           | 300                         | 15                                         | 0.4                   | 25                   |
|                                  | PH <sub>3</sub> (against SiH <sub>4</sub> )                                                 | 50 ppm           |                             |                                            |                       |                      |
| Upper layer                      | 3rd layer region                                                                            | SiH <sub>4</sub> | 100                         |                                            |                       |                      |
|                                  | layer region                                                                                | H <sub>2</sub>   | 300                         | 5                                          | 0.2                   | 8                    |
|                                  | 4th layer region                                                                            | SiH <sub>4</sub> | 100                         |                                            |                       |                      |
|                                  | NH <sub>3</sub>                                                                             | 80→100*          | 300                         | 5                                          | 0.4                   | 0.7                  |
|                                  | B <sub>2</sub> H <sub>6</sub> (against SiH <sub>4</sub> )                                   | 500 ppm          |                             |                                            |                       |                      |

TABLE 61

| Order of lamination<br>(layer name) | Gases and<br>their flow rates<br>(SCCM)                                                                                                 | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|-----------------------------------------------------------------------------------------------------------------------------------------|-----------------------------------|--------------------------------------------------|-----------------------------|----------------------------|
| Lower layer                         | SiH <sub>4</sub> 50<br>H <sub>2</sub> 5→200*<br>AlCl <sub>3</sub> /He<br>(S-side: 0.01 μm)<br>(UL-side: 0.01 μm)<br>200→30**<br>30→10** | 250                               | 1                                                | 0.3                         | 0.02                       |
| 1st<br>layer                        | B <sub>2</sub> H <sub>6</sub> (against SiH <sub>4</sub> ) 100 ppm<br>SiH <sub>4</sub> 100                                               | 250                               | 10                                               | 0.4                         | 3                          |
| Upper<br>layer                      | He 600<br>SiH <sub>4</sub> 300<br>He 600<br>B <sub>2</sub> H <sub>6</sub> 0.5 ppm<br>SiH <sub>4</sub> 50<br>CH <sub>4</sub> 500         | 250                               | 25                                               | 0.6                         | 25                         |
| 2nd<br>layer                        |                                                                                                                                         | 250                               | 10                                               | 0.4                         | 1                          |
| 3rd<br>layer                        |                                                                                                                                         |                                   |                                                  |                             |                            |
| region                              |                                                                                                                                         |                                   |                                                  |                             |                            |

TABLE 62

| Order of lamination<br>(layer name) | Gases and<br>their flow rates<br>(SCCM)                                                                                                                                                                                                                                                                                                                                               | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|---------------------------------------------------------------------------------------------------------------------------------------------------------------------------------------------------------------------------------------------------------------------------------------------------------------------------------------------------------------------------------------|-----------------------------------|--------------------------------------------------|-----------------------------|----------------------------|
| Lower layer                         | SiH <sub>4</sub> 10→100*<br>H <sub>2</sub> 5→200*<br>AlCl <sub>3</sub> /He<br>(S-side: 0.05 μm)<br>(UL-side: 0.15 μm)<br>200→40**<br>40→10**                                                                                                                                                                                                                                          | 300                               | 10                                               | 0.4                         | 0.2                        |
| 1st<br>layer                        | B <sub>2</sub> H <sub>6</sub> (against SiH <sub>4</sub> ) 50 ppm<br>SiH <sub>4</sub> 100<br>B <sub>2</sub> H <sub>6</sub> 200 ppm<br>H <sub>2</sub> 500<br>SiF <sub>4</sub> 0.5<br>AlCl <sub>3</sub> /He 0.1<br>SiH <sub>4</sub> 300                                                                                                                                                  | 300                               | 8                                                | 0.4                         | 0.5                        |
| Upper<br>layer                      | H <sub>2</sub> 500<br>CH <sub>4</sub> 1<br>NO 0.1<br>B <sub>2</sub> H <sub>6</sub> 0.3 ppm<br>SiF <sub>4</sub> 0.5<br>AlCl <sub>3</sub> /He 0.1<br>SiH <sub>4</sub> 100<br>CH <sub>4</sub> 600<br>PH <sub>3</sub> (against SiH <sub>4</sub> ) 3000 ppm<br>NO 0.1<br>SiF <sub>4</sub> 0.5<br>AlCl <sub>3</sub> /He 0.1<br>B <sub>2</sub> H <sub>6</sub> 0.3 ppm<br>SiH <sub>4</sub> 40 | 300                               | 20                                               | 0.5                         | 20                         |
| 2nd<br>layer                        |                                                                                                                                                                                                                                                                                                                                                                                       |                                   |                                                  |                             |                            |
| region                              |                                                                                                                                                                                                                                                                                                                                                                                       |                                   |                                                  |                             |                            |
| 3rd<br>layer                        |                                                                                                                                                                                                                                                                                                                                                                                       |                                   |                                                  |                             |                            |
| region                              |                                                                                                                                                                                                                                                                                                                                                                                       |                                   |                                                  |                             |                            |
| 4th<br>layer                        |                                                                                                                                                                                                                                                                                                                                                                                       |                                   |                                                  |                             |                            |
| region                              |                                                                                                                                                                                                                                                                                                                                                                                       |                                   |                                                  |                             |                            |
|                                     |                                                                                                                                                                                                                                                                                                                                                                                       |                                   |                                                  |                             |                            |

TABLE 63

| Order of lamination<br>(layer name) | Gases and<br>their flow rates<br>(SCCM)                                                                                                                                                                           | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|-------------------------------------------------------------------------------------------------------------------------------------------------------------------------------------------------------------------|-----------------------------------|--------------------------------------------------|-----------------------------|----------------------------|
| Lower layer                         | SiH <sub>4</sub> 10→100*<br>H <sub>2</sub> 5→200*<br>AlCl <sub>3</sub> /He<br>(S-side: 0.5 μm)<br>(UL-side: 0.15 μm)<br>200→40**<br>40→10**                                                                       | 250                               | 5                                                | 0.4                         | 0.2                        |
| 1st<br>layer                        | B <sub>2</sub> H <sub>6</sub> (against SiH <sub>4</sub> ) 100 ppm<br>SiH <sub>4</sub> 100<br>B <sub>2</sub> H <sub>6</sub> (against SiH <sub>4</sub> )<br>(LL-side: 2 μm)<br>(U · 2nd · LR-side:<br>1 μm) 500 ppm | 250                               | 8                                                | 0.4                         | 3                          |

TABLE 63-continued

| Order of lamination<br>(layer name) | Gases and their flow rates<br>(SCCM)                                            | Substrate temperature<br>(°C.)                                                                                                                                                 | RF discharging power<br>(mW/cm <sup>3</sup> )  | Inner pressure<br>(Torr) | Layer thickness<br>(μm) |     |
|-------------------------------------|---------------------------------------------------------------------------------|--------------------------------------------------------------------------------------------------------------------------------------------------------------------------------|------------------------------------------------|--------------------------|-------------------------|-----|
| region                              | 500<br>ppm—0**                                                                  |                                                                                                                                                                                |                                                |                          |                         |     |
|                                     | H <sub>2</sub><br>SiF <sub>4</sub><br>AlCl <sub>3</sub> /He<br>SiH <sub>4</sub> | 200<br>0.5<br>0.1<br>100                                                                                                                                                       |                                                |                          |                         |     |
| Upper layer                         | 2nd layer                                                                       | SiF <sub>4</sub><br>H <sub>2</sub><br>CH <sub>4</sub><br>NO<br>B <sub>2</sub> H <sub>6</sub> (against SiH <sub>4</sub> )<br>AlCl <sub>3</sub> /He<br>SiH <sub>4</sub>          | 5<br>200<br>1<br>0.1<br>0.3 ppm<br>0.1<br>100  | 300                      | 3<br>0.5                | 3   |
|                                     | region                                                                          | CH <sub>4</sub><br>NO<br>B <sub>2</sub> H <sub>6</sub> (against SiH <sub>4</sub> )<br>AlCl <sub>3</sub> /He<br>SiH <sub>4</sub>                                                | 100<br>50 ppm<br>0.1<br>0.3 ppm<br>0.5         | 300                      | 15<br>0.4               | 30  |
|                                     | 3rd layer                                                                       | CH <sub>4</sub><br>PH <sub>3</sub> (against SiH <sub>4</sub> )<br>NO<br>B <sub>2</sub> H <sub>6</sub> (against SiH <sub>4</sub> )<br>AlCl <sub>3</sub> /He<br>SiH <sub>4</sub> | 100<br>50 ppm<br>0.1<br>0.3 ppm<br>0.1<br>50   | 300                      | 10<br>0.4               | 0.5 |
|                                     | region                                                                          | CH <sub>4</sub><br>PH <sub>3</sub> (against SiH <sub>4</sub> )<br>B <sub>2</sub> H <sub>6</sub> (against SiH <sub>4</sub> )<br>NO<br>SiF <sub>4</sub><br>AlCl <sub>3</sub> /He | 600<br>0.3 ppm<br>0.3 ppm<br>0.1<br>0.5<br>0.1 | 300                      |                         |     |
|                                     | 4th layer                                                                       | CH <sub>4</sub><br>PH <sub>3</sub> (against SiH <sub>4</sub> )<br>B <sub>2</sub> H <sub>6</sub> (against SiH <sub>4</sub> )<br>NO<br>SiF <sub>4</sub><br>AlCl <sub>3</sub> /He | 600<br>0.3 ppm<br>0.1<br>0.5<br>0.1            |                          |                         |     |

TABLE 64

| Order of lamination<br>(layer name) | Gases and their flow rates<br>(SCCM)                                                                                             | Substrate temperature<br>(°C.)                                                                                                                                                             | RF discharging power<br>(mW/cm <sup>3</sup> )                  | Inner pressure<br>(Torr) | Layer thickness<br>(μm) |  |
|-------------------------------------|----------------------------------------------------------------------------------------------------------------------------------|--------------------------------------------------------------------------------------------------------------------------------------------------------------------------------------------|----------------------------------------------------------------|--------------------------|-------------------------|--|
| Lower layer                         | H <sub>2</sub> S (against SiH <sub>4</sub> )<br>SiH <sub>4</sub><br>H <sub>2</sub><br>AlCl <sub>3</sub> /He<br>(S-side: 0.05 μm) | 3 ppm<br>10→100*<br>5→200*<br>300                                                                                                                                                          | 10                                                             | 0.4                      | 0.2                     |  |
|                                     |                                                                                                                                  | 200→40**                                                                                                                                                                                   |                                                                |                          |                         |  |
|                                     | (UL-side: 0.15 μm)                                                                                                               | 40→10**                                                                                                                                                                                    |                                                                |                          |                         |  |
|                                     | B <sub>2</sub> H <sub>6</sub> (against SiH <sub>4</sub> )<br>SiH <sub>4</sub>                                                    | 50 ppm<br>100                                                                                                                                                                              |                                                                |                          |                         |  |
| 1st layer                           | region                                                                                                                           | B <sub>2</sub> H <sub>6</sub><br>H <sub>2</sub><br>SiF <sub>4</sub><br>AlCl <sub>3</sub> /He<br>H <sub>2</sub> S<br>SiH <sub>4</sub><br>H <sub>2</sub>                                     | 200 ppm<br>500<br>0.5<br>0.1<br>1 ppm<br>300<br>500            | 300<br>8                 | 0.4<br>0.5              |  |
| Upper layer                         | 2nd layer                                                                                                                        | CH <sub>4</sub><br>NO<br>B <sub>2</sub> H <sub>6</sub><br>SiF <sub>4</sub><br>AlCl <sub>3</sub> /He<br>H <sub>2</sub> S<br>SiH <sub>4</sub><br>CH <sub>4</sub>                             | 1<br>0.1<br>0.3 ppm<br>0.5<br>0.1<br>1 ppm<br>100<br>600       | 300<br>20                | 0.5<br>20               |  |
|                                     | region                                                                                                                           | PH <sub>3</sub> (against SiH <sub>4</sub> )<br>NO<br>SiF <sub>4</sub><br>AlCl <sub>3</sub> /He<br>B <sub>2</sub> H <sub>6</sub><br>H <sub>2</sub> S<br>SiH <sub>4</sub><br>CH <sub>4</sub> | 3000 ppm<br>0.1<br>0.5<br>0.1<br>0.3 ppm<br>1 ppm<br>40<br>600 | 300<br>15                | 0.4<br>7                |  |
|                                     | 3rd layer                                                                                                                        | NO<br>SiF <sub>4</sub><br>AlCl <sub>3</sub> /He<br>B <sub>2</sub> H <sub>6</sub><br>H <sub>2</sub> S<br>SiH <sub>4</sub><br>CH <sub>4</sub>                                                | 0.1<br>0.5<br>0.1<br>0.3 ppm<br>1 ppm<br>40<br>600             | 300                      |                         |  |
|                                     | region                                                                                                                           | NO<br>PH <sub>3</sub><br>B <sub>2</sub> H <sub>6</sub><br>SiF <sub>4</sub><br>AlCl <sub>3</sub> /He<br>H <sub>2</sub> S                                                                    | 0.1<br>0.3 ppm<br>0.5<br>0.1<br>1 ppm                          | 300<br>10                | 0.4<br>0.1              |  |
|                                     | 4th layer                                                                                                                        | NO<br>PH <sub>3</sub><br>B <sub>2</sub> H <sub>6</sub><br>SiF <sub>4</sub><br>AlCl <sub>3</sub> /He<br>H <sub>2</sub> S                                                                    | 0.1<br>0.3 ppm<br>0.5<br>0.1<br>1 ppm                          |                          |                         |  |

TABLE 65

| Order of lamination (layer name) | Gases and their flow rates (SCCM) |                                                           | Substrate temperature (°C.) | RF discharging power (mW/cm <sup>3</sup> ) | Inner pressure (Torr) | Layer thickness (μm) |
|----------------------------------|-----------------------------------|-----------------------------------------------------------|-----------------------------|--------------------------------------------|-----------------------|----------------------|
| Lower layer                      | SiH <sub>4</sub>                  | 50                                                        | 250                         | 5                                          | 0.4                   | 0.05                 |
|                                  | NO                                | 5                                                         |                             |                                            |                       |                      |
|                                  | H <sub>2</sub>                    | 10→200*                                                   |                             |                                            |                       |                      |
|                                  | AlCl <sub>3</sub> /He             | 120→40**                                                  | 250                         | 8                                          | 0.4                   | 3                    |
|                                  | 1st layer region                  | SiH <sub>4</sub>                                          |                             |                                            |                       |                      |
|                                  | 2nd layer region                  | B <sub>2</sub> H <sub>6</sub> (against SiH <sub>4</sub> ) | 200 ppm                     |                                            |                       |                      |
| Upper layer                      | 3rd layer region                  | H <sub>2</sub>                                            | 500                         | 250                                        | 15                    | 0.5                  |
|                                  | 2nd layer region                  | SiH <sub>4</sub>                                          | 300                         |                                            |                       |                      |
|                                  | 1st layer region                  | H <sub>2</sub>                                            | 300                         |                                            |                       |                      |
|                                  | 3rd layer region                  | SiH <sub>4</sub>                                          | 50                          | 250                                        | 10                    | 0.4                  |
|                                  | 2nd layer region                  | CH <sub>4</sub>                                           | 500                         |                                            |                       |                      |
|                                  | 1st layer region                  |                                                           |                             |                                            |                       |                      |

TABLE 66

| Order of lamination (layer name) | Gases and their flow rates (SCCM) |                                                           | Substrate temperature (°C.) | RF discharging power (mW/cm <sup>3</sup> ) | Inner pressure (Torr) | Layer thickness (μm) |
|----------------------------------|-----------------------------------|-----------------------------------------------------------|-----------------------------|--------------------------------------------|-----------------------|----------------------|
| Lower layer                      | SiH <sub>4</sub>                  | 50                                                        | 250                         | 5                                          | 0.4                   | 0.05                 |
|                                  | AlCl <sub>3</sub> /He             | 120→40**                                                  |                             |                                            |                       |                      |
|                                  | 1st layer region                  | SiH <sub>4</sub>                                          |                             |                                            |                       |                      |
|                                  | 2nd layer region                  | B <sub>2</sub> H <sub>6</sub> (against SiH <sub>4</sub> ) | 200 ppm                     | 250                                        | 8                     | 0.4                  |
|                                  | 3rd layer region                  | H <sub>2</sub>                                            | 500                         | 250                                        | 15                    | 0.5                  |
|                                  | 2nd layer region                  | SiH <sub>4</sub>                                          | 300                         |                                            |                       |                      |
| Upper layer                      | 1st layer region                  | H <sub>2</sub>                                            | 300                         |                                            |                       |                      |
|                                  | 2nd layer region                  | SiH <sub>4</sub>                                          | 50                          | 250                                        | 10                    | 0.4                  |
|                                  | 3rd layer region                  | CH <sub>4</sub>                                           | 500                         |                                            |                       |                      |
|                                  | 2nd layer region                  |                                                           |                             |                                            |                       |                      |
|                                  | 1st layer region                  |                                                           |                             |                                            |                       |                      |
|                                  |                                   |                                                           |                             |                                            |                       |                      |

TABLE 67

| Order of lamination (layer name) | Gases and their flow rates (SCCM)       |                                                           | Substrate temperature (°C.) | RF discharging power (mW/cm <sup>3</sup> ) | Inner pressure (Torr) | Layer thickness (μm) |
|----------------------------------|-----------------------------------------|-----------------------------------------------------------|-----------------------------|--------------------------------------------|-----------------------|----------------------|
| Lower layer                      | SiH <sub>4</sub>                        | 50                                                        | 250                         | 5                                          | 0.4                   | 0.03                 |
|                                  | NO                                      | 5                                                         |                             |                                            |                       |                      |
|                                  | H <sub>2</sub>                          | 10→200*                                                   |                             |                                            |                       |                      |
|                                  | AlCl <sub>3</sub> /He (S-side: 0.01 μm) | 100→10**                                                  | 250                         | 8                                          | 0.4                   | 3                    |
|                                  | 1st layer region                        | (UL-side: 0.01 μm)                                        |                             |                                            |                       |                      |
|                                  | 2nd layer region                        | SiH <sub>4</sub>                                          | 100                         |                                            |                       |                      |
| Upper layer                      | 3rd layer region                        | B <sub>2</sub> H <sub>6</sub> (against SiH <sub>4</sub> ) | 200 ppm                     | 250                                        | 15                    | 0.5                  |
|                                  | 2nd layer region                        | H <sub>2</sub>                                            | 500                         | 250                                        | 10                    | 0.5                  |
|                                  | 1st layer region                        | SiH <sub>4</sub>                                          | 300                         |                                            |                       |                      |
|                                  | 3rd layer region                        | H <sub>2</sub>                                            | 300                         |                                            |                       |                      |
|                                  | 2nd layer region                        | SiH <sub>4</sub>                                          | 50                          | 250                                        | 0.4                   | 0.5                  |
|                                  | 1st layer region                        | CH <sub>4</sub>                                           | 500                         |                                            |                       |                      |

TABLE 68

| Order of lamination (layer name) | Gases and their flow rates (SCCM)                         |                                                                           | Substrate temperature (°C.) | RF discharging power (mW/cm <sup>3</sup> ) | Inner pressure (Torr) | Layer thickness (μm) |  |  |
|----------------------------------|-----------------------------------------------------------|---------------------------------------------------------------------------|-----------------------------|--------------------------------------------|-----------------------|----------------------|--|--|
| Lower layer                      | B <sub>2</sub> H <sub>6</sub> (against SiH <sub>4</sub> ) | 30 ppm                                                                    | 150                         | 0.5                                        | 0.3                   | 0.02                 |  |  |
|                                  | SiH <sub>4</sub>                                          | 50                                                                        |                             |                                            |                       |                      |  |  |
|                                  | H <sub>2</sub>                                            | 5→200*                                                                    |                             |                                            |                       |                      |  |  |
|                                  | AlCl <sub>3</sub> /He (S-side: 0.01 μm)                   | 200→30**                                                                  | 300                         | 1.5                                        | 0.4                   | 3                    |  |  |
|                                  | 1st layer region                                          | (UL-side: 0.01 μm)                                                        | 30→10**                     | 250                                        |                       |                      |  |  |
|                                  | 2nd layer region                                          | NO                                                                        | 5                           |                                            |                       |                      |  |  |
| Upper layer                      | 3rd layer region                                          | SiH <sub>4</sub>                                                          | 100                         | 10                                         | 0.4                   | 3                    |  |  |
|                                  | 2nd layer region                                          | B <sub>2</sub> H <sub>6</sub> (against SiH <sub>4</sub> ) (LL-side: 2 μm) | 500 ppm                     |                                            |                       |                      |  |  |
|                                  | 1st layer region                                          | (U·2nd·LR-side: 1 μm)                                                     | 500 ppm                     |                                            |                       |                      |  |  |
|                                  | 3rd layer region                                          | H <sub>2</sub>                                                            | 200 ppm→0**                 | 250                                        | 0.4                   | 0.5                  |  |  |
|                                  | 2nd layer region                                          |                                                                           |                             |                                            |                       |                      |  |  |
|                                  | 1st layer region                                          |                                                                           |                             |                                            |                       |                      |  |  |

TABLE 68-continued

| Order of lamination (layer name) | Gases and their flow rates (SCCM)  |            | Substrate temperature (°C.) | RF discharging power (mW/cm <sup>3</sup> ) | Inner pressure (Torr) | Layer thickness (μm) |
|----------------------------------|------------------------------------|------------|-----------------------------|--------------------------------------------|-----------------------|----------------------|
| 2nd layer region                 | SiH <sub>4</sub><br>H <sub>2</sub> | 300<br>500 | 250                         | 20                                         | 0.5                   | 20                   |

TABLE 69

| Order of lamination (layer name) | Gases and their flow rates (SCCM)                         |          | Substrate temperature (°C.) | RF discharging power (mW/cm <sup>3</sup> ) | Inner pressure (Torr) | Layer thickness (μm) |
|----------------------------------|-----------------------------------------------------------|----------|-----------------------------|--------------------------------------------|-----------------------|----------------------|
| Lower layer                      | SiH <sub>4</sub>                                          | 50       | 250                         | 1                                          | 0.3                   | 0.02                 |
|                                  | H <sub>2</sub>                                            | 5→200*   |                             |                                            |                       |                      |
|                                  | AlCl <sub>3</sub> /He<br>(S-side: 0.01 μm)                | 200→30** |                             |                                            |                       |                      |
|                                  | (UL-side: 0.01 μm)                                        | 30→10**  |                             |                                            |                       |                      |
|                                  | N <sub>2</sub>                                            | 100      |                             |                                            |                       |                      |
|                                  | SiH <sub>4</sub>                                          | 100      |                             |                                            |                       |                      |
|                                  | B <sub>2</sub> H <sub>6</sub> (against SiH <sub>4</sub> ) | 500 ppm  |                             |                                            |                       |                      |
|                                  | He                                                        | 600      |                             |                                            |                       |                      |
|                                  | AlCl <sub>3</sub> /He                                     | 0.1      |                             |                                            |                       |                      |
|                                  | SiF <sub>4</sub>                                          | 0.5      |                             |                                            |                       |                      |
| Upper layer                      | NO                                                        | 0.1      | 250                         | 10                                         | 0.4                   | 3                    |
|                                  | CH <sub>4</sub>                                           | 1        |                             |                                            |                       |                      |
|                                  | SiH <sub>4</sub>                                          | 300      |                             |                                            |                       |                      |
|                                  | He                                                        | 600      |                             |                                            |                       |                      |
|                                  | B <sub>2</sub> H <sub>6</sub>                             | 0.3 ppm  |                             |                                            |                       |                      |
|                                  | SiF <sub>4</sub>                                          | 0.5      |                             |                                            |                       |                      |
|                                  | AlCl <sub>3</sub> /He                                     | 0.1      |                             |                                            |                       |                      |
|                                  | SiH <sub>4</sub>                                          | 50       |                             |                                            |                       |                      |
|                                  | CH <sub>4</sub>                                           | 500      |                             |                                            |                       |                      |
|                                  | NO                                                        | 0.1      |                             |                                            |                       |                      |
| 3rd layer region                 | B <sub>2</sub> H <sub>6</sub>                             | 0.3 ppm  | 10                          | 0.6                                        | 25                    | 1                    |
|                                  | SiF <sub>4</sub>                                          | 0.5      |                             |                                            |                       |                      |
|                                  | AlCl <sub>3</sub> /He                                     | 0.1      |                             |                                            |                       |                      |
|                                  | SiH <sub>4</sub>                                          | 0.1      |                             |                                            |                       |                      |

TABLE 70

| Order of lamination (layer name) | Gases and their flow rates (SCCM)                                                                            |             | Substrate temperature (°C.) | RF discharging power (mW/cm <sup>3</sup> ) | Inner pressure (Torr) | Layer thickness (μm) |
|----------------------------------|--------------------------------------------------------------------------------------------------------------|-------------|-----------------------------|--------------------------------------------|-----------------------|----------------------|
| Lower layer                      | SiH <sub>4</sub>                                                                                             | 10→100*     | 250                         | 10                                         | 0.4                   | 0.2                  |
|                                  | H <sub>2</sub>                                                                                               | 5→200*      |                             |                                            |                       |                      |
|                                  | AlCl <sub>3</sub> /He<br>(S-side: 0.05 μm)                                                                   | 200→40**    |                             |                                            |                       |                      |
|                                  | (UL-side: 0.15 μm)                                                                                           | 40→10**     |                             |                                            |                       |                      |
|                                  | CH <sub>4</sub>                                                                                              | 50→200*     |                             |                                            |                       |                      |
|                                  | SiH <sub>4</sub>                                                                                             | 100         |                             |                                            |                       |                      |
|                                  | B <sub>2</sub> H <sub>6</sub> (against SiH <sub>4</sub> )<br>(LL-side: 2 μm)<br>(U + 2nd -LR-sided:<br>1 μm) | 500 ppm     |                             |                                            |                       |                      |
|                                  |                                                                                                              | 500 ppm→0** |                             |                                            |                       |                      |
|                                  | H <sub>2</sub>                                                                                               | 200         |                             |                                            |                       |                      |
|                                  | SiH <sub>4</sub>                                                                                             | 400         |                             |                                            |                       |                      |
| 2nd layer region                 | Ar                                                                                                           | 200         | 250                         | 10                                         | 0.5                   | 15                   |
|                                  | SiH <sub>4</sub>                                                                                             | 100         |                             |                                            |                       |                      |
|                                  | NH <sub>3</sub>                                                                                              | 30          |                             |                                            |                       |                      |
| 3rd layer region                 |                                                                                                              |             |                             |                                            |                       |                      |

TABLE 71

| Order of lamination (layer name) | Gases and their flow rates (SCCM)                                                |                   | Substrate temperature (°C.) | RF discharging power (mW/cm <sup>3</sup> ) | Inner pressure (Torr) | Layer thickness (μm) |
|----------------------------------|----------------------------------------------------------------------------------|-------------------|-----------------------------|--------------------------------------------|-----------------------|----------------------|
| Lower layer                      | SiH <sub>4</sub><br>H <sub>2</sub><br>AlCl <sub>3</sub> /He<br>(S-side: 0.05 μm) | 10→100*<br>5→200* | 300                         | 10                                         | 0.4                   | 0.2                  |

TABLE 71-continued

| Order of lamination<br>(layer name) | Gases and their flow rates<br>(SCCM)        | Substrate temperature<br>(°C.) | RF discharging power<br>(mW/cm <sup>3</sup> ) | Inner pressure<br>(Torr) | Layer thickness<br>(μm) |
|-------------------------------------|---------------------------------------------|--------------------------------|-----------------------------------------------|--------------------------|-------------------------|
| Upper layer                         | NO                                          | 40→10**                        |                                               |                          |                         |
|                                     | SiH <sub>4</sub>                            | 5→20                           |                                               |                          |                         |
|                                     | B <sub>2</sub> H <sub>6</sub>               | 100                            |                                               |                          |                         |
|                                     | H <sub>2</sub>                              | 200 ppm                        | 300                                           | 8                        | 0.4                     |
|                                     |                                             | 500                            |                                               |                          |                         |
|                                     | SiH <sub>4</sub>                            | 300                            |                                               |                          |                         |
|                                     | H <sub>2</sub>                              | 500                            | 300                                           | 20                       | 0.5                     |
|                                     |                                             |                                |                                               |                          |                         |
|                                     | SiH <sub>4</sub>                            | 100                            |                                               |                          |                         |
|                                     | CH <sub>4</sub>                             | 600                            | 300                                           | 15                       | 0.4                     |
| region                              | PH <sub>3</sub> (against SiH <sub>4</sub> ) | 3000 ppm                       |                                               |                          |                         |
|                                     | SiH <sub>4</sub>                            | 40                             |                                               |                          |                         |
|                                     | CH <sub>4</sub>                             | 600                            | 300                                           | 10                       | 0.4                     |
|                                     |                                             |                                |                                               |                          | 0.1                     |
| region                              |                                             |                                |                                               |                          |                         |

TABLE 72

| Order of lamination<br>(layer name) | Gases and their flow rates<br>(SCCM)        | Substrate temperature<br>(°C.) | RF discharging power<br>(mW/cm <sup>3</sup> ) | Inner pressure<br>(Torr) | Layer thickness<br>(μm) |
|-------------------------------------|---------------------------------------------|--------------------------------|-----------------------------------------------|--------------------------|-------------------------|
| Lower layer                         | PH <sub>3</sub> (against SiH <sub>4</sub> ) | 20 ppm                         |                                               |                          |                         |
|                                     | SiH <sub>4</sub>                            | 50                             |                                               |                          |                         |
|                                     | H <sub>2</sub>                              | 5→200*                         | 330                                           | 5                        | 0.4                     |
|                                     | AlCl <sub>3</sub> /He                       | 200→20**                       |                                               |                          |                         |
|                                     | NO                                          | 5                              |                                               |                          |                         |
|                                     | SiH <sub>4</sub>                            | 100                            |                                               |                          |                         |
|                                     | PH <sub>3</sub>                             | 100 ppm                        | 330                                           | 8                        | 0.4                     |
|                                     | H <sub>2</sub>                              | 100                            |                                               |                          |                         |
|                                     | SiF <sub>4</sub>                            | 400                            |                                               |                          |                         |
|                                     | H <sub>2</sub>                              | 800                            | 330                                           | 25                       | 0.5                     |
| Upper layer                         | SiH <sub>4</sub>                            | 100                            |                                               |                          |                         |
|                                     | SiF <sub>4</sub>                            | 400                            |                                               |                          |                         |
|                                     | H <sub>2</sub>                              | 800                            | 350                                           | 15                       | 0.4                     |
|                                     | CH <sub>4</sub>                             | 400                            |                                               |                          |                         |
|                                     | B <sub>2</sub> H <sub>6</sub>               | 5000 ppm                       |                                               |                          |                         |
|                                     | SiH <sub>4</sub>                            | 20                             |                                               |                          |                         |
|                                     | CH <sub>4</sub>                             | 400                            | 350                                           | 10                       | 0.4                     |
|                                     | B <sub>2</sub> H <sub>6</sub>               | 8000 ppm                       |                                               |                          | 1                       |
|                                     |                                             |                                |                                               |                          |                         |

TABLE 73

| Order of lamination<br>(layer name) | Gases and their flow rates<br>(SCCM)                      | Substrate temperature<br>(°C.) | RF discharging power<br>(mW/cm <sup>3</sup> ) | Inner pressure<br>(Torr) | Layer thickness<br>(μm) |
|-------------------------------------|-----------------------------------------------------------|--------------------------------|-----------------------------------------------|--------------------------|-------------------------|
| Lower layer                         | SiH <sub>4</sub>                                          | 50                             |                                               |                          |                         |
|                                     | H <sub>2</sub> S (against SiH <sub>4</sub> )              | 10 ppm                         |                                               |                          |                         |
|                                     | B <sub>2</sub> H <sub>6</sub> (against SiH <sub>4</sub> ) | 30 ppm                         |                                               |                          |                         |
|                                     | H <sub>2</sub>                                            | 5→200*                         | 300                                           | 1                        | 0.3                     |
|                                     | AlCl <sub>3</sub> /He<br>(S-side: 0.01 μm)                | 200→30**                       |                                               |                          |                         |
|                                     | (UL-side: 0.01 μm)                                        | 30→10**                        |                                               |                          |                         |
|                                     | CH <sub>4</sub>                                           | 50                             |                                               |                          |                         |
|                                     | SiH <sub>4</sub>                                          | 100                            |                                               |                          |                         |
|                                     | B <sub>2</sub> H <sub>6</sub> (against SiH <sub>4</sub> ) | 200 ppm                        | 300                                           | 8                        | 0.4                     |
|                                     | H <sub>2</sub>                                            | 500                            |                                               |                          |                         |
| Upper layer                         | SiH <sub>4</sub>                                          | 300                            |                                               |                          |                         |
|                                     | SiH <sub>4</sub>                                          | 300                            | 20                                            | 0.5                      | 20                      |
|                                     | B <sub>2</sub> H <sub>6</sub>                             | 200                            |                                               |                          |                         |
|                                     | SiH <sub>4</sub>                                          | 50                             |                                               |                          |                         |
|                                     | N <sub>2</sub>                                            | 500                            | 300                                           | 20                       | 0.4                     |
|                                     | PH <sub>3</sub> (against SiH <sub>4</sub> )               | 3000 ppm                       |                                               |                          |                         |
|                                     | SiH <sub>4</sub>                                          | 40                             |                                               |                          |                         |
|                                     | CH <sub>4</sub>                                           | 600                            | 300                                           | 10                       | 0.4                     |
|                                     |                                                           |                                |                                               |                          | 0.3                     |

TABLE 74

| Order of lamination<br>(layer name) | Gases and their flow rates<br>(SCCM)                      | Substrate temperature<br>(°C.) | RF discharging power<br>(mW/cm <sup>3</sup> ) | Inner pressure<br>(Torr) | Layer thickness<br>(μm) |
|-------------------------------------|-----------------------------------------------------------|--------------------------------|-----------------------------------------------|--------------------------|-------------------------|
|                                     | B <sub>2</sub> H <sub>6</sub> (against SiH <sub>4</sub> ) | 50 ppm                         |                                               |                          |                         |

TABLE 74-continued

| Order of lamination<br>(layer name) | Gases and their flow rates (SCCM)                                            |                | Substrate temperature (°C.) | RF discharging power (mW/cm <sup>3</sup> ) | Inner pressure (Torr) | Layer thickness (μm) |
|-------------------------------------|------------------------------------------------------------------------------|----------------|-----------------------------|--------------------------------------------|-----------------------|----------------------|
| Lower layer                         | SiH <sub>4</sub>                                                             | 50             | 250                         | 5                                          | 0.4                   | 0.05                 |
|                                     | H <sub>2</sub>                                                               | 5→200*         |                             |                                            |                       |                      |
|                                     | AlCl <sub>3</sub> /He                                                        | 200→20**       |                             |                                            |                       |                      |
|                                     | NO                                                                           | 5              |                             |                                            |                       |                      |
|                                     | C <sub>2</sub> H <sub>2</sub>                                                | 10             |                             |                                            |                       |                      |
|                                     | SiH <sub>4</sub>                                                             | 100            |                             |                                            |                       |                      |
| 1st layer                           | B <sub>2</sub> H <sub>6</sub> (against SiH <sub>4</sub> )<br>(LL-side: 3 μm) | 500 ppm        | 250                         | 10                                         | 0.4                   | 5                    |
|                                     | (U + 2nd + LR-side:<br>2 μm)                                                 |                |                             |                                            |                       |                      |
| Upper region<br>layer               |                                                                              | 500<br>ppm→0** |                             |                                            |                       |                      |
|                                     | H <sub>2</sub>                                                               | 200            |                             |                                            |                       |                      |
|                                     | AlCl <sub>3</sub> /He (against<br>SiH <sub>4</sub> )                         | 1→0**          |                             |                                            |                       |                      |
| 2nd layer region                    | SiH <sub>4</sub>                                                             | 300            | 250                         | 15                                         | 0.5                   | 10                   |
|                                     | H <sub>2</sub>                                                               | 300            |                             |                                            |                       |                      |
| 3rd layer region                    | SiH <sub>4</sub>                                                             | 200            | 250                         | 15                                         | 0.4                   | 20                   |
|                                     | C <sub>2</sub> H <sub>2</sub>                                                | 10→20*         |                             |                                            |                       |                      |
| NO                                  | 1                                                                            |                |                             |                                            |                       |                      |

TABLE 75

| Order of lamination<br>(layer name) | Gases and their flow rates (SCCM)                                            |                | Substrate temperature (°C.) | RF discharging power (mW/cm <sup>3</sup> ) | Inner pressure (Torr) | Layer thickness (μm) |
|-------------------------------------|------------------------------------------------------------------------------|----------------|-----------------------------|--------------------------------------------|-----------------------|----------------------|
| Lower layer                         | NO                                                                           | 5              | 250                         | 1                                          | 0.4                   | 0.02                 |
|                                     | SiH <sub>4</sub>                                                             | 50             |                             |                                            |                       |                      |
|                                     | H <sub>2</sub>                                                               | 5→200*         |                             |                                            |                       |                      |
|                                     | AlCl <sub>3</sub> /He<br>(S-side: 0.01 μm)                                   | 200→30**       |                             |                                            |                       |                      |
|                                     | (UL-side: 0.01 μm)                                                           | 30→10**        |                             |                                            |                       |                      |
|                                     | H <sub>2</sub> S (against SiH <sub>4</sub> )                                 | 10 ppm         |                             |                                            |                       |                      |
| 1st layer region                    | SiH <sub>4</sub>                                                             | 100            | 250                         | 10                                         | 0.4                   | 10                   |
|                                     | B <sub>2</sub> H <sub>6</sub> (against SiH <sub>4</sub> )<br>(LL-side: 2 μm) | 500 ppm        |                             |                                            |                       |                      |
|                                     | (U + 2nd + LR-side:<br>1 μm)                                                 |                |                             |                                            |                       |                      |
|                                     |                                                                              | 500<br>ppm→0** |                             |                                            |                       |                      |
| Upper layer                         | H <sub>2</sub>                                                               | 200            | 300                         | 20                                         | 0.5                   | 5                    |
|                                     | SiH <sub>4</sub>                                                             | 300            |                             |                                            |                       |                      |
|                                     | H <sub>2</sub>                                                               | 300            |                             |                                            |                       |                      |
|                                     | SiH <sub>4</sub>                                                             | 100            |                             |                                            |                       |                      |
|                                     | CH <sub>4</sub>                                                              | 100            |                             | 15                                         | 0.4                   | 20                   |
|                                     | SiH <sub>4</sub>                                                             | 50             |                             |                                            |                       |                      |
|                                     | CH <sub>4</sub>                                                              | 600            |                             | 10                                         | 0.4                   | 0.5                  |

TABLE 76

| Order of lamination<br>(layer name) | Gases and their flow rates (SCCM)                         |          | Substrate temperature (°C.) | RF discharging power (mW/cm <sup>3</sup> ) | Inner pressure (Torr) | Layer thickness (μm) |
|-------------------------------------|-----------------------------------------------------------|----------|-----------------------------|--------------------------------------------|-----------------------|----------------------|
| Lower layer                         | SiH <sub>4</sub>                                          | 10→100*  | 300                         | 5                                          | 0.4                   | 0.2                  |
|                                     | H <sub>2</sub>                                            | 5→200*   |                             |                                            |                       |                      |
|                                     | AlCl <sub>3</sub> /He<br>(S-side: 0.05 μm)                | 200→40** |                             |                                            |                       |                      |
|                                     | (UL-side: 0.15 μm)                                        | 40→10**  |                             |                                            |                       |                      |
|                                     | NH <sub>3</sub>                                           | 5→50*    |                             |                                            |                       |                      |
|                                     | SiH <sub>4</sub>                                          | 100      |                             |                                            |                       |                      |
| Upper layer                         | B <sub>2</sub> H <sub>6</sub> (against SiH <sub>4</sub> ) | 200 ppm  | 300                         | 5                                          | 0.4                   | 3                    |
|                                     | H <sub>2</sub>                                            | 500      |                             |                                            |                       |                      |
|                                     | SiH <sub>4</sub>                                          | 100      |                             |                                            |                       |                      |
|                                     | H <sub>2</sub>                                            | 300      |                             |                                            |                       |                      |
| 2nd layer region                    | SiH <sub>4</sub>                                          | 300      | 300                         | 5                                          | 0.2                   | 8                    |
|                                     | NH <sub>3</sub>                                           | 50       |                             |                                            |                       |                      |
| 3rd layer                           | SiH <sub>4</sub>                                          | 300      | 300                         | 15                                         | 0.4                   | 25                   |
|                                     | NH <sub>3</sub>                                           | 50       |                             |                                            |                       |                      |

TABLE 76-continued

| Order of lamination<br>(layer name) | Gases and their flow rates (SCCM) |     | Substrate temperature (°C.) | RF discharging power (mW/cm <sup>3</sup> ) | Inner pressure (Torr) | Layer thickness (μm) |
|-------------------------------------|-----------------------------------|-----|-----------------------------|--------------------------------------------|-----------------------|----------------------|
| region                              |                                   |     |                             |                                            |                       |                      |
| 4th layer region                    | SiH <sub>4</sub>                  | 100 | 300                         | 10                                         | 0.4                   | 0.3                  |
|                                     | NH <sub>3</sub>                   | 50  |                             |                                            |                       |                      |

TABLE 77

| Order of lamination<br>(layer name) | Gases and their flow rates (SCCM)                                            |               | Substrate temperature (°C.) | RF discharging power (mW/cm <sup>3</sup> ) | Inner pressure (Torr) | Layer thickness (μm) |
|-------------------------------------|------------------------------------------------------------------------------|---------------|-----------------------------|--------------------------------------------|-----------------------|----------------------|
| Lower layer                         | SiH <sub>4</sub>                                                             | 10 → 100*     |                             |                                            |                       |                      |
|                                     | H <sub>2</sub>                                                               | 5 → 200*      |                             |                                            |                       |                      |
|                                     | AlCl <sub>3</sub> /He<br>(S-side: 0.05 μm)                                   |               | 250                         | 5                                          | 0.4                   | 0.2                  |
|                                     |                                                                              | 200 → 40**    |                             |                                            |                       |                      |
|                                     | (UL-side: 0.15 μm)                                                           |               |                             |                                            |                       |                      |
|                                     | NO                                                                           | 40 → 10**     |                             |                                            |                       |                      |
| 1st layer region                    | SiH <sub>4</sub>                                                             | 5 → 20        |                             |                                            |                       |                      |
|                                     | B <sub>2</sub> H <sub>6</sub> (against SiH <sub>4</sub> )<br>(LL-side: 2 μm) | 100           |                             |                                            |                       |                      |
|                                     | (U · 2nd · LR-side: 1 μm)                                                    | 500 ppm       | 250                         | 8                                          | 0.4                   | 3                    |
|                                     |                                                                              | 500 ppm → 0** |                             |                                            |                       |                      |
| Upper layer                         | H <sub>2</sub>                                                               | 200           |                             |                                            |                       |                      |
| 2nd layer region                    | SiH <sub>4</sub>                                                             | 100           |                             |                                            |                       |                      |
|                                     | SiF <sub>4</sub>                                                             | 5             | 300                         | 3                                          | 0.5                   | 3                    |
| 3rd layer region                    | H <sub>2</sub>                                                               | 200           |                             |                                            |                       |                      |
|                                     | SiH <sub>4</sub>                                                             | 100           |                             |                                            |                       |                      |
| 4th layer region                    | CH <sub>4</sub>                                                              | 100           | 300                         | 15                                         | 0.4                   | 30                   |
|                                     | PH <sub>3</sub> (against SiH <sub>4</sub> )                                  | 50 ppm        |                             |                                            |                       |                      |
|                                     | SiH <sub>4</sub>                                                             | 50            |                             |                                            |                       |                      |
|                                     | CH <sub>4</sub>                                                              | 600           | 300                         | 10                                         | 0.4                   | 0.5                  |

TABLE 78

| Order of lamination<br>(layer name) | Gases and their flow rates (SCCM)                                                      |               | Substrate temperature (°C.) | RF discharging power (mW/cm <sup>3</sup> ) | Inner pressure (Torr) | Layer thickness (μm) |
|-------------------------------------|----------------------------------------------------------------------------------------|---------------|-----------------------------|--------------------------------------------|-----------------------|----------------------|
| Lower layer                         | N <sub>2</sub>                                                                         | 300           |                             |                                            |                       |                      |
|                                     | SiH <sub>4</sub>                                                                       | 50            |                             |                                            |                       |                      |
|                                     | H <sub>2</sub>                                                                         | 5 → 200*      | 250                         | 5                                          | 0.4                   | 0.05                 |
|                                     | AlCl <sub>3</sub> /He                                                                  | 200 → 20**    |                             |                                            |                       |                      |
|                                     | PH <sub>3</sub> (against SiH <sub>4</sub> )                                            | 50 ppm        |                             |                                            |                       |                      |
| 1st layer region                    | SiH <sub>4</sub>                                                                       | 40            |                             |                                            |                       |                      |
|                                     | PH <sub>3</sub> (against SiH <sub>4</sub> )<br>(LL-side: 2 μm)                         | 250 ppm       | 250                         | 8                                          | 0.4                   | 3                    |
|                                     | (U · 2nd · LR-side: 1 μm)                                                              | 250 ppm → 0** |                             |                                            |                       |                      |
| Upper layer                         | H <sub>2</sub>                                                                         | 40            |                             |                                            |                       |                      |
| 2nd layer region                    | Si <sub>2</sub> H <sub>6</sub>                                                         | 200           |                             |                                            |                       |                      |
|                                     | H <sub>2</sub>                                                                         | 200           | 300                         | 10                                         | 0.5                   | 10                   |
| 3rd layer region                    | SiH <sub>4</sub>                                                                       | 300           |                             |                                            |                       |                      |
|                                     | C <sub>2</sub> H <sub>2</sub>                                                          | 50            |                             |                                            |                       |                      |
|                                     | B <sub>2</sub> H <sub>6</sub> (against SiH <sub>4</sub> )<br>(U · 2nd · LR-side: 1 μm) | 0 → 100 ppm*  | 330                         | 20                                         | 0.4                   | 30                   |
|                                     | (U · 4th · LR-side: 29 μm)                                                             | 100 ppm       |                             |                                            |                       |                      |
| 4th layer region                    | SiH <sub>4</sub>                                                                       | 200           |                             |                                            |                       |                      |
|                                     | C <sub>2</sub> H <sub>2</sub>                                                          | 200           | 330                         | 10                                         | 0.4                   | 1                    |

TABLE 79

| Order of lamination<br>(layer name) | Gases and their flow rates (SCCM)                         |           | Substrate temperature (°C.) | RF discharging power (mW/cm <sup>3</sup> ) | Inner pressure (Torr) | Layer thickness (μm) |
|-------------------------------------|-----------------------------------------------------------|-----------|-----------------------------|--------------------------------------------|-----------------------|----------------------|
| Lower layer                         | B <sub>2</sub> H <sub>6</sub> (against SiH <sub>4</sub> ) | 100 ppm   |                             |                                            |                       |                      |
|                                     | SiH <sub>4</sub>                                          | 10 → 100* |                             |                                            |                       |                      |
|                                     | H <sub>2</sub>                                            | 5 → 200*  |                             |                                            |                       |                      |
|                                     | AlCl <sub>3</sub> /He<br>(S-side: 0.05 μm)                |           | 250                         | 5                                          | 0.4                   | 0.2                  |

TABLE 79-continued

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Upper layer                      | 200 → 40**<br>(UL-side: 0.15 μm)                          |                             |                                            |                       |                      |
|                                  | NO                                                        | 50 → 200*                   |                                            |                       |                      |
|                                  | SiH <sub>4</sub>                                          | 100                         |                                            |                       |                      |
|                                  | B <sub>2</sub> H <sub>6</sub> (against SiH <sub>4</sub> ) | 200 ppm                     | 300                                        | 8                     | 0.3                  |
|                                  | H <sub>2</sub>                                            | 500                         |                                            |                       |                      |
|                                  | SiH <sub>4</sub>                                          | 100                         |                                            |                       |                      |
|                                  | H <sub>2</sub>                                            | 300                         | 300                                        | 5                     | 0.2                  |
|                                  | SiH <sub>4</sub>                                          | 300                         |                                            |                       |                      |
|                                  | NH <sub>3</sub>                                           | 30 → 50*                    | 300                                        | 15                    | 0.4                  |
|                                  | PH <sub>3</sub> (against SiH <sub>4</sub> )               | 50 ppm                      |                                            |                       |                      |
| Upper layer                      | SiH <sub>4</sub>                                          | 100                         |                                            |                       |                      |
|                                  | NH <sub>3</sub>                                           | 80 → 100*                   | 300                                        | 5                     | 0.4                  |
| Upper layer                      | PH <sub>3</sub> (against SiH <sub>4</sub> )               | 500 ppm                     |                                            |                       | 0.7                  |

TABLE 80

| Order of lamination (layer name) | Gases and their flow rates (SCCM) | Substrate temperature (°C.) | RF discharging power (mW/cm <sup>3</sup> ) | Inner pressure (Torr) | Layer thickness (μm) |
|----------------------------------|-----------------------------------|-----------------------------|--------------------------------------------|-----------------------|----------------------|
| Upper layer                      | SiH <sub>4</sub>                  | 50                          |                                            |                       |                      |
|                                  | H <sub>2</sub>                    | 5 → 200*                    |                                            |                       |                      |
|                                  | AlCl <sub>3</sub> /He             |                             | 250                                        | 1                     | 0.4                  |
|                                  | (S-side: 0.01 μm)                 |                             |                                            |                       |                      |
|                                  | 200 → 30**<br>(UL-side: 0.01 μm)  |                             |                                            |                       |                      |
|                                  | NO                                | 30 → 10**                   |                                            |                       |                      |
|                                  | SiH <sub>4</sub>                  | 10                          |                                            |                       |                      |
|                                  | PH <sub>3</sub>                   | 100 ppm                     | 300                                        | 8                     | 0.4                  |
|                                  | H <sub>2</sub>                    | 100                         |                                            |                       |                      |
|                                  | SiH <sub>4</sub>                  | 300                         |                                            |                       |                      |
| Upper layer                      | H <sub>2</sub>                    | 500                         | 300                                        | 20                    | 0.5                  |
|                                  | SiH <sub>4</sub>                  | 100                         |                                            |                       |                      |
|                                  | GeH <sub>4</sub>                  | 10 → 50*                    | 300                                        | 5                     | 0.4                  |
|                                  | H <sub>2</sub>                    | 300                         |                                            |                       |                      |
|                                  | SiH <sub>4</sub>                  | 100 → 40**                  |                                            |                       |                      |
| Upper layer                      | CH <sub>4</sub>                   | 100 → 600*                  | 300                                        | 10                    | 0.4                  |
|                                  |                                   |                             |                                            |                       | 1                    |

TABLE 81

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Upper layer                      | B <sub>2</sub> H <sub>6</sub> (against SiH <sub>4</sub> ) | 70 ppm                      |                                            |                       |                      |
|                                  | SiH <sub>4</sub>                                          | 50                          |                                            |                       |                      |
|                                  | H <sub>2</sub>                                            | 5 → 200*                    |                                            |                       |                      |
|                                  | AlCl <sub>3</sub> /He                                     |                             | 300                                        | 1                     | 0.3                  |
|                                  | (S-side: 0.01 μm)                                         |                             |                                            |                       |                      |
|                                  | 200 → 30**<br>(UL-side: 0.01 μm)                          |                             |                                            |                       |                      |
|                                  | NO                                                        | 30 → 10**                   |                                            |                       |                      |
|                                  | SiH <sub>4</sub>                                          | 5                           |                                            |                       |                      |
|                                  | SiH <sub>4</sub>                                          | 100                         |                                            |                       |                      |
|                                  | B <sub>2</sub> H <sub>6</sub> (against SiH <sub>4</sub> ) | 200 ppm                     | 300                                        | 8                     | 0.4                  |
| Upper layer                      | H <sub>2</sub>                                            | 500                         |                                            |                       |                      |
|                                  | SiH <sub>4</sub>                                          | 300                         |                                            |                       |                      |
|                                  | H <sub>2</sub>                                            | 400                         | 300                                        | 15                    | 0.5                  |
|                                  | SiH <sub>4</sub>                                          | 50                          |                                            |                       |                      |
| Upper layer                      | CH <sub>4</sub>                                           | 500                         | 300                                        | 10                    | 0.4                  |
|                                  |                                                           |                             |                                            |                       | 0.5                  |

TABLE 82

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 50                                               |                             |                                            |                       |                      |
|                                  | B <sub>2</sub> H <sub>6</sub> (against SiH <sub>4</sub> ) 50 ppm  |                             |                                            |                       |                      |
|                                  | NO 5                                                              |                             |                                            |                       |                      |
|                                  | H <sub>2</sub> 5 → 200*                                           | 300                         | 0.7                                        | 0.3                   | 0.02                 |
|                                  | AlCl <sub>3</sub> /He (S-side: 0.01 μm)                           |                             |                                            |                       |                      |
|                                  | (UL-side: 0.01 μm) 200 → 30**                                     |                             |                                            |                       |                      |
| 1st layer region                 | SiH <sub>4</sub> 80                                               |                             |                                            |                       |                      |
|                                  | H <sub>2</sub> 400                                                | 300                         | 7                                          | 0.3                   | 10                   |
|                                  | B <sub>2</sub> H <sub>6</sub> (against SiH <sub>4</sub> ) 200 ppm |                             |                                            |                       |                      |
| Upper layer                      | 2nd layer region SiH <sub>4</sub> 200                             |                             |                                            |                       |                      |
|                                  | H <sub>2</sub> 400                                                | 300                         | 12                                         | 0.4                   | 20                   |
|                                  | 3rd layer region SiH <sub>4</sub> 40                              |                             |                                            |                       |                      |
|                                  | CH <sub>4</sub> 400                                               | 300                         | 7                                          | 0.3                   | 0.5                  |
|                                  | B <sub>2</sub> H <sub>6</sub> (against SiH <sub>4</sub> ) 200 ppm |                             |                                            |                       |                      |
|                                  |                                                                   |                             |                                            |                       |                      |

TABLE 83

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 25                                               |                             |                                            |                       |                      |
|                                  | B <sub>2</sub> H <sub>6</sub> (against SiH <sub>4</sub> ) 50 ppm  |                             |                                            |                       |                      |
|                                  | NO 3                                                              |                             |                                            |                       |                      |
|                                  | H <sub>2</sub> 5 → 100*                                           | 300                         | 0.5                                        | 0.2                   | 0.02                 |
|                                  | AlCl <sub>3</sub> /He (S-side: 0.01 μm)                           |                             |                                            |                       |                      |
|                                  | (UL-side: 0.01 μm) 100 → 15**                                     |                             |                                            |                       |                      |
| 1st layer region                 | SiH <sub>4</sub> 60                                               |                             |                                            |                       |                      |
|                                  | H <sub>2</sub> 300                                                | 300                         | 6                                          | 0.2                   | 10                   |
|                                  | B <sub>2</sub> H <sub>6</sub> (against SiH <sub>4</sub> ) 200 ppm |                             |                                            |                       |                      |
| Upper layer                      | 2nd layer region SiH <sub>4</sub> 150                             |                             |                                            |                       |                      |
|                                  | H <sub>2</sub> 300                                                | 300                         | 10                                         | 0.4                   | 20                   |
|                                  | 3rd layer region SiH <sub>4</sub> 30                              |                             |                                            |                       |                      |
|                                  | CH <sub>4</sub> 300                                               | 300                         | 5                                          | 0.3                   | 0.5                  |
|                                  | B <sub>2</sub> H <sub>6</sub> (against SiH <sub>4</sub> ) 200 ppm |                             |                                            |                       |                      |
|                                  |                                                                   |                             |                                            |                       |                      |

TABLE 84

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 20                                               |                             |                                            |                       |                      |
|                                  | B <sub>2</sub> H <sub>6</sub> (against SiH <sub>4</sub> ) 50 ppm  |                             |                                            |                       |                      |
|                                  | NO 2                                                              | 300                         | 0.3                                        | 0.2                   | 0.02                 |
|                                  | H <sub>2</sub> 5 → 100*                                           |                             |                                            |                       |                      |
|                                  | AlCl <sub>3</sub> /He (S-side: 0.01 μm)                           |                             |                                            |                       |                      |
|                                  | (UL-side: 0.01 μm) 80 → 15**                                      |                             |                                            |                       |                      |
| 1st layer region                 | SiH <sub>4</sub> 40                                               |                             |                                            |                       |                      |
|                                  | H <sub>2</sub> 200                                                | 300                         | 5                                          | 0.2                   | 10                   |
|                                  | B <sub>2</sub> H <sub>6</sub> (against SiH <sub>4</sub> ) 200 ppm |                             |                                            |                       |                      |
| Upper layer                      | 2nd layer region SiH <sub>4</sub> 100                             |                             |                                            |                       |                      |
|                                  | H <sub>2</sub> 300                                                | 300                         | 6                                          | 0.3                   | 20                   |
|                                  | 3rd layer region SiH <sub>4</sub> 20                              |                             |                                            |                       |                      |
|                                  | CH <sub>4</sub> 200                                               | 300                         | 3                                          | 0.2                   | 0.5                  |
|                                  | B <sub>2</sub> H <sub>6</sub> (against SiH <sub>4</sub> ) 200 ppm |                             |                                            |                       |                      |
|                                  |                                                                   |                             |                                            |                       |                      |

TABLE 85

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 50                          |                                            |                       |                      |
|                                  | B <sub>2</sub> H <sub>6</sub> (against SiH <sub>4</sub> ) | 100 ppm                     |                                            |                       |                      |
|                                  | NO                                                        | 5                           | 500                                        | 5                     | 0.4                  |
|                                  | H <sub>2</sub>                                            | 5 → 200*                    |                                            |                       |                      |
|                                  | AlCl <sub>3</sub> /He                                     | 200 → 20**                  |                                            |                       |                      |
|                                  | SiH <sub>4</sub>                                          | 100                         |                                            |                       |                      |
| 1st layer region                 | B <sub>2</sub> H <sub>6</sub> (against SiH <sub>4</sub> ) |                             |                                            |                       |                      |
|                                  | (LL-side: 2 μm)<br>(U · 2nd · LR-side: 1 μm)              | 500 ppm                     | 500                                        | 20                    | 0.4                  |
| Upper layer                      |                                                           | 500 → 0 ppm**               |                                            |                       |                      |
|                                  | H <sub>2</sub>                                            | 1200                        |                                            |                       |                      |
|                                  | 2nd layer region                                          | SiH <sub>4</sub>            | 300                                        |                       |                      |
|                                  | H <sub>2</sub>                                            | 1500                        | 500                                        | 30                    | 0.5                  |
| 3rd layer region                 | SiH <sub>4</sub>                                          | 200                         |                                            |                       |                      |
|                                  | C <sub>2</sub> H <sub>2</sub>                             | 10 → 20*                    | 500                                        | 30                    | 0.4                  |
|                                  | NO                                                        | 1                           |                                            |                       | 20                   |

TABLE 86

| Order of lamination (layer name) | Gases and their flow rates (SCCM)                         | Substrate temperature (°C.) | μW discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | B <sub>2</sub> H <sub>6</sub> (against SiH <sub>4</sub> ) | 50 ppm                      |                                            |                       |                      |
|                                  | SiH <sub>4</sub>                                          | 150                         |                                            |                       |                      |
|                                  | H <sub>2</sub>                                            | 20 → 500*                   |                                            |                       |                      |
|                                  | AlCl <sub>3</sub> /He<br>(S-side: 0.01 μm)                | 250                         | 0.5                                        | 0.6                   | 0.02                 |
|                                  | (UL-side: 0.01 μm)                                        | 400 → 80**                  |                                            |                       |                      |
|                                  |                                                           | 80 → 50**                   |                                            |                       |                      |
| Upper layer                      | NO                                                        | 10                          |                                            |                       |                      |
|                                  | SiH <sub>4</sub>                                          | 100                         |                                            |                       |                      |
|                                  | B <sub>2</sub> H <sub>6</sub> (against SiH <sub>4</sub> ) | 200 ppm                     | 250                                        | 0.5                   | 0.5                  |
|                                  | H <sub>2</sub>                                            | 500                         |                                            |                       | 3                    |
|                                  | 2nd layer region                                          | SiH <sub>4</sub>            | 700                                        |                       |                      |
|                                  | SiF <sub>4</sub>                                          | 30                          | 250                                        | 0.5                   | 0.5                  |
| 3rd layer region                 | H <sub>2</sub>                                            | 500                         |                                            |                       | 20                   |
|                                  | SiH <sub>4</sub>                                          | 150                         |                                            |                       |                      |
|                                  | CH <sub>4</sub>                                           | 500                         | 250                                        | 0.5                   | 0.3                  |
|                                  |                                                           |                             |                                            |                       | 1                    |

TABLE 87

| Order of lamination (layer name) | Gases and their flow rates (SCCM)                                                                         | Substrate temperature (°C.) | RF discharging power (mW/cm <sup>3</sup> ) | Inner pressure (Torr) | Layer thickness (μm) |
|----------------------------------|-----------------------------------------------------------------------------------------------------------|-----------------------------|--------------------------------------------|-----------------------|----------------------|
| Lower layer                      | B <sub>2</sub> H <sub>6</sub> (against SiH <sub>4</sub> )                                                 | 50 ppm                      |                                            |                       |                      |
|                                  | SiH <sub>4</sub>                                                                                          | 50                          |                                            |                       |                      |
|                                  | H <sub>2</sub>                                                                                            | 5 → 200*                    | 250                                        | 5                     | 0.4                  |
|                                  | AlCl <sub>3</sub> /He                                                                                     | 200 → 20**                  |                                            |                       |                      |
|                                  | NO                                                                                                        | 5                           |                                            |                       |                      |
|                                  | C <sub>2</sub> H <sub>2</sub>                                                                             | 10                          |                                            |                       |                      |
| 1st layer region                 | SiH <sub>4</sub>                                                                                          | 100                         |                                            |                       |                      |
|                                  | B <sub>2</sub> H <sub>6</sub> (against SiH <sub>4</sub> )<br>(LL-side: 3 μm)<br>(U · 2nd · LR-side: 2 μm) | 500 ppm                     | 250                                        | 10                    | 0.4                  |
| Upper layer                      |                                                                                                           | 500 ppm → 0**               |                                            |                       |                      |
|                                  | H <sub>2</sub>                                                                                            | 200                         |                                            |                       |                      |
|                                  | AlCl <sub>3</sub> /He<br>(against SiH <sub>4</sub> )                                                      | 1 → 0**                     |                                            |                       |                      |
|                                  | SiH <sub>4</sub>                                                                                          | 200                         |                                            |                       |                      |
|                                  | C <sub>2</sub> H <sub>2</sub>                                                                             | 10 → 20*                    | 250                                        | 15                    | 0.4                  |
|                                  | NO                                                                                                        | 1                           |                                            |                       | 20                   |
| 3rd layer region                 | SiH <sub>4</sub>                                                                                          | 300                         |                                            |                       |                      |
|                                  | H <sub>2</sub>                                                                                            | 300                         | 250                                        | 15                    | 0.5                  |
|                                  |                                                                                                           |                             |                                            |                       | 10                   |

TABLE 88

| Order of lamination<br>(layer name) | Gases and their flow rates<br>(SCCM)                                         | Substrate temperature<br>(°C.) | RF discharging power<br>(mW/cm <sup>3</sup> ) | Inner pressure<br>(Torr) | Layer thickness<br>(μm) |
|-------------------------------------|------------------------------------------------------------------------------|--------------------------------|-----------------------------------------------|--------------------------|-------------------------|
| Lower layer                         | NO                                                                           | 5                              |                                               |                          |                         |
|                                     | SiH <sub>4</sub>                                                             | 50                             |                                               |                          |                         |
|                                     | H <sub>2</sub>                                                               | 5 → 200*                       |                                               |                          |                         |
|                                     | AlCl <sub>3</sub> /He<br>(S-side: 0.01 μm)                                   | 250                            | 1                                             | 0.4                      | 0.02                    |
|                                     | (UL-side: 0.01 μm)                                                           | 200 → 30**                     |                                               |                          |                         |
|                                     | H <sub>2</sub> S (against SiH <sub>4</sub> )                                 | 30 → 10**                      |                                               |                          |                         |
|                                     | SiH <sub>4</sub>                                                             | 10 ppm                         |                                               |                          |                         |
|                                     | B <sub>2</sub> H <sub>6</sub> (against SiH <sub>4</sub> )<br>(LL-side: 2 μm) | 100                            |                                               |                          |                         |
|                                     | (U + 2nd + LR-side: 1 μm)                                                    | 500 ppm                        | 250                                           | 10                       | 0.4                     |
|                                     |                                                                              | 500 ppm → 0**                  |                                               | 10                       |                         |
| Upper layer                         | H <sub>2</sub>                                                               | 200                            |                                               |                          |                         |
|                                     | SiH <sub>4</sub>                                                             | 100                            |                                               |                          |                         |
|                                     | CH <sub>4</sub>                                                              | 100                            | 300                                           | 15                       | 0.4                     |
|                                     | SiH <sub>4</sub>                                                             | 300                            | 300                                           | 20                       | 0.5                     |
|                                     | H <sub>2</sub>                                                               | 300                            |                                               |                          | 5                       |
|                                     | SiH <sub>4</sub>                                                             | 50                             | 300                                           | 10                       | 0.4                     |
|                                     | CH <sub>4</sub>                                                              | 600                            |                                               |                          | 0.5                     |

TABLE 89

| Order of lamination<br>(layer name) | Gases and their flow rates<br>(SCCM)                      | Substrate temperature<br>(°C.) | RF discharging power<br>(mW/cm <sup>3</sup> ) | Inner pressure<br>(Torr) | Layer thickness<br>(μm) |
|-------------------------------------|-----------------------------------------------------------|--------------------------------|-----------------------------------------------|--------------------------|-------------------------|
| Lower layer                         | SiH <sub>4</sub>                                          | 10 → 100*                      |                                               |                          |                         |
|                                     | H <sub>2</sub>                                            | 5 → 200*                       |                                               |                          |                         |
|                                     | AlCl <sub>3</sub> /He<br>(S-side: 0.05 μm)                | 300                            | 5                                             | 0.4                      | 0.2                     |
|                                     | (UL-side: 0.15 μm)                                        | 200 → 40**                     |                                               |                          |                         |
|                                     |                                                           | 40 → 10**                      |                                               |                          |                         |
|                                     | NH <sub>3</sub>                                           | 5 → 50*                        |                                               |                          |                         |
|                                     | SiH <sub>4</sub>                                          | 100                            |                                               |                          |                         |
|                                     | B <sub>2</sub> H <sub>6</sub> (against SiH <sub>4</sub> ) | 200 ppm                        | 300                                           | 5                        | 0.4                     |
|                                     | H <sub>2</sub>                                            | 500                            |                                               |                          | 3                       |
|                                     |                                                           |                                |                                               |                          |                         |
| Upper layer                         | SiH <sub>4</sub>                                          | 300                            |                                               |                          |                         |
|                                     | NH <sub>3</sub>                                           | 50                             | 300                                           | 15                       | 0.4                     |
|                                     | SiH <sub>4</sub>                                          | 100                            |                                               |                          |                         |
|                                     | H <sub>2</sub>                                            | 300                            | 300                                           | 5                        | 0.2                     |
|                                     | SiH <sub>4</sub>                                          | 100                            |                                               |                          | 8                       |
|                                     | NH <sub>3</sub>                                           | 50                             | 300                                           | 10                       | 0.4                     |
|                                     |                                                           |                                |                                               |                          | 0.3                     |

TABLE 90

| Order of lamination<br>(layer name) | Gases and their flow rates<br>(SCCM)        | Substrate temperature<br>(°C.) | RF discharging power<br>(mW/cm <sup>3</sup> ) | Inner pressure<br>(Torr) | Layer thickness<br>(μm) |
|-------------------------------------|---------------------------------------------|--------------------------------|-----------------------------------------------|--------------------------|-------------------------|
| Lower layer                         | SiH <sub>4</sub>                            | 10 → 100*                      |                                               |                          |                         |
|                                     | H <sub>2</sub>                              | 5 → 200*                       |                                               |                          |                         |
|                                     | AlCl <sub>3</sub> /He<br>(S-side: 0.05 μm)  | 250                            | 5                                             | 0.4                      | 0.2                     |
|                                     | (UL-side: 0.15 μm)                          | 200 → 40**                     |                                               |                          |                         |
|                                     |                                             | 40 → 10**                      |                                               |                          |                         |
|                                     | NO                                          | 5 → 20                         |                                               |                          |                         |
|                                     | SiH <sub>4</sub>                            | 100                            |                                               |                          |                         |
|                                     | PH <sub>3</sub> (against SiH <sub>4</sub> ) | 100 ppm                        | 250                                           | 8                        | 0.4                     |
|                                     | H <sub>2</sub>                              | 100                            |                                               |                          | 3                       |
|                                     |                                             |                                |                                               |                          |                         |
| Upper layer                         | SiH <sub>4</sub>                            | 100                            |                                               |                          |                         |
|                                     | CH <sub>4</sub>                             | 100                            | 300                                           | 10                       | 0.4                     |
|                                     | PH <sub>3</sub> (against SiH <sub>4</sub> ) | 50 ppm                         |                                               |                          | 30                      |
|                                     | SiH <sub>4</sub>                            | 100                            |                                               |                          |                         |
|                                     | SiF <sub>4</sub>                            | 5                              | 300                                           | 3                        | 0.5                     |
|                                     | H <sub>2</sub>                              | 200                            |                                               |                          | 3                       |
|                                     | SiH <sub>4</sub>                            | 50                             |                                               |                          |                         |

TABLE 90-continued

| Order of lamination (layer name) | Gases and their flow rates (SCCM) | Substrate temperature (°C.) | RF discharging power (mW/cm <sup>3</sup> ) | Inner pressure (Torr) | Layer thickness (μm) |
|----------------------------------|-----------------------------------|-----------------------------|--------------------------------------------|-----------------------|----------------------|
| layer region                     | CH <sub>4</sub> 600               | 300                         | 10                                         | 0.4                   | 0.5                  |

TABLE 91

| Order of lamination (layer name) | Gases and their flow rates (SCCM)                                                   | Substrate temperature (°C.) | RF discharging power (mW/cm <sup>3</sup> ) | Inner pressure (Torr) | Layer thickness (μm) |
|----------------------------------|-------------------------------------------------------------------------------------|-----------------------------|--------------------------------------------|-----------------------|----------------------|
| Lower layer                      | N <sub>2</sub> 300                                                                  | 250                         | 5                                          | 0.4                   | 0.05                 |
|                                  | SiH <sub>4</sub> 50                                                                 |                             |                                            |                       |                      |
|                                  | H <sub>2</sub> 5 → 200*                                                             |                             |                                            |                       |                      |
|                                  | AlCl <sub>3</sub> /He 200 → 20**                                                    |                             |                                            |                       |                      |
|                                  | B <sub>2</sub> H <sub>6</sub> (against SiH <sub>4</sub> ) 50 ppm                    |                             |                                            |                       |                      |
| 1st layer region                 | SiH <sub>4</sub> 100                                                                | 250                         | 8                                          | 0.4                   | 3                    |
|                                  | B <sub>2</sub> H <sub>6</sub> (against SiH <sub>4</sub> ) (LL-side: 2 μm) 500 ppm   |                             |                                            |                       |                      |
|                                  | (U · 2nd · LR-side: 1 μm)                                                           |                             |                                            |                       |                      |
| Upper layer                      | H <sub>2</sub> 500 ppm → 0**                                                        | 330                         | 20                                         | 0.4                   | 30                   |
|                                  | SiH <sub>4</sub> 200                                                                |                             |                                            |                       |                      |
|                                  | C <sub>2</sub> H <sub>2</sub> 300                                                   |                             |                                            |                       |                      |
|                                  | B <sub>2</sub> H <sub>6</sub> (against SiH <sub>4</sub> ) (U · 1st · LR-side: 1 μm) |                             |                                            |                       |                      |
|                                  | (U · 3rd · LR-side: 29 μm)                                                          |                             |                                            |                       |                      |
| 3rd layer region                 | Si <sub>2</sub> H <sub>6</sub> 100 ppm                                              | 300                         | 10                                         | 0.5                   | 10                   |
|                                  | H <sub>2</sub> 200                                                                  |                             |                                            |                       |                      |
| 4th layer region                 | SiH <sub>4</sub> 200                                                                | 330                         | 10                                         | 0.4                   | 1                    |
|                                  | C <sub>2</sub> H <sub>2</sub> 200                                                   |                             |                                            |                       |                      |

TABLE 92

| Order of lamination (layer name) | Gases and their flow rates (SCCM)                                   | Substrate temperature (°C.) | RF discharging power (mW/cm <sup>3</sup> ) | Inner pressure (Torr) | Layer thickness (μm) |
|----------------------------------|---------------------------------------------------------------------|-----------------------------|--------------------------------------------|-----------------------|----------------------|
| Lower layer                      | PH <sub>3</sub> (against SiH <sub>4</sub> ) 50 ppm                  | 250                         | 5                                          | 0.4                   | 0.2                  |
|                                  | SiH <sub>4</sub> 10 → 100*                                          |                             |                                            |                       |                      |
|                                  | H <sub>2</sub> 5 → 200*                                             |                             |                                            |                       |                      |
|                                  | AlCl <sub>3</sub> /He (S-side: 0.05 μm) 200 → 40**                  |                             |                                            |                       |                      |
|                                  | (UL-side: 0.15 μm)                                                  |                             |                                            |                       |                      |
| 1st layer region                 | NO 40 → 10**                                                        | 250                         | 8                                          | 0.4                   | 3                    |
|                                  | SiH <sub>4</sub> 20 → 200*                                          |                             |                                            |                       |                      |
|                                  | PH <sub>3</sub> (against SiH <sub>4</sub> ) (LL-side: 2 μm) 250 ppm |                             |                                            |                       |                      |
| Upper layer                      | (U · 2nd · LR-side: 1 μm)                                           | 300                         | 15                                         | 0.4                   | 25                   |
|                                  | H <sub>2</sub> 250 ppm → 0**                                        |                             |                                            |                       |                      |
|                                  | SiH <sub>4</sub> 40                                                 |                             |                                            |                       |                      |
|                                  | NH <sub>3</sub> 30 → 50*                                            |                             |                                            |                       |                      |
|                                  | PH <sub>3</sub> (against SiH <sub>4</sub> ) 50 ppm                  |                             |                                            |                       |                      |
| 3rd layer region                 | SiH <sub>4</sub> 100                                                | 300                         | 5                                          | 0.2                   | 8                    |
|                                  | H <sub>2</sub> 300                                                  |                             |                                            |                       |                      |
|                                  | NH <sub>3</sub> 30 → 50*                                            |                             |                                            |                       |                      |
|                                  | PH <sub>3</sub> (against SiH <sub>4</sub> ) 50 ppm                  |                             |                                            |                       |                      |
| 4th layer region                 | H <sub>2</sub> 300                                                  | 300                         | 5                                          | 0.4                   | 0.7                  |
|                                  | SiH <sub>4</sub> 100                                                |                             |                                            |                       |                      |
| NH <sub>3</sub> region           | NH <sub>3</sub> 80 → 100*                                           | 300                         | 5                                          | 0.4                   | 0.7                  |
|                                  | B <sub>2</sub> H <sub>6</sub> (against SiH <sub>4</sub> ) 500 ppm   |                             |                                            |                       |                      |

TABLE 93

| Order of lamination (layer name)        | Gases and their flow rates (SCCM)                  | Substrate temperature (°C.) | RF discharging power (mW/cm <sup>3</sup> ) | Inner pressure (Torr) | Layer thickness (μm) |
|-----------------------------------------|----------------------------------------------------|-----------------------------|--------------------------------------------|-----------------------|----------------------|
| Lower layer                             | SiH <sub>4</sub> 50                                | 250                         | 1                                          | 0.3                   | 0.02                 |
|                                         | H <sub>2</sub> 5 → 200*                            |                             |                                            |                       |                      |
| AlCl <sub>3</sub> /He (S-side: 0.01 μm) | AlCl <sub>3</sub> /He (S-side: 0.01 μm) 200 → 30** |                             |                                            |                       |                      |
|                                         | (UL-side: 0.01 μm)                                 |                             |                                            |                       |                      |

TABLE 93-continued

| Order of lamination (layer name) | Gases and their flow rates (SCCM) |                                                           | Substrate temperature (°C.) | RF discharging power (mW/cm <sup>3</sup> ) | Inner pressure (Torr) | Layer thickness (μm) |
|----------------------------------|-----------------------------------|-----------------------------------------------------------|-----------------------------|--------------------------------------------|-----------------------|----------------------|
| Upper layer                      | 1st layer region                  | N <sub>2</sub>                                            | 30 → 10**                   |                                            |                       |                      |
|                                  |                                   | SiH <sub>4</sub>                                          | 100                         |                                            |                       |                      |
|                                  |                                   | B <sub>2</sub> H <sub>6</sub> (against SiH <sub>4</sub> ) | 100                         |                                            |                       |                      |
|                                  | 2nd layer region                  | He                                                        | 500 ppm                     | 250                                        | 10                    | 0.4                  |
|                                  |                                   | He                                                        | 600                         |                                            |                       | 3                    |
|                                  |                                   | B <sub>2</sub> H <sub>6</sub>                             | 0.5 ppm                     |                                            |                       |                      |
| Lower layer                      | 3rd layer region                  | SiH <sub>4</sub>                                          | 300                         |                                            |                       |                      |
|                                  | SiH <sub>4</sub>                  | 600                                                       | 250                         | 25                                         | 0.6                   | 25                   |
|                                  | CH <sub>4</sub>                   | 500                                                       |                             | 10                                         | 0.4                   | 1                    |

TABLE 94

| Order of lamination (layer name) | Gases and their flow rates (SCCM) |                                             | Substrate temperature (°C.) | RF discharging power (mW/cm <sup>3</sup> ) | Inner pressure (Torr) | Layer thickness (μm) |
|----------------------------------|-----------------------------------|---------------------------------------------|-----------------------------|--------------------------------------------|-----------------------|----------------------|
| Upper layer                      | 1st layer region                  | SiH <sub>4</sub>                            | 10 → 100*                   |                                            |                       |                      |
|                                  |                                   | H <sub>2</sub>                              | 5 → 200*                    |                                            |                       |                      |
|                                  |                                   | AlCl <sub>3</sub> /He (S-side: 0.05 μm)     | 300                         | 10                                         | 0.4                   | 0.2                  |
|                                  | 2nd layer region                  | SiH <sub>4</sub>                            | 200 → 40**                  |                                            |                       |                      |
|                                  |                                   | NO                                          | 40 → 10**                   |                                            |                       |                      |
|                                  |                                   | SiH <sub>4</sub>                            | 5 → 20                      |                                            |                       |                      |
| Lower layer                      | 3rd layer region                  | B <sub>2</sub> H <sub>6</sub>               | 100                         |                                            |                       |                      |
|                                  |                                   | H <sub>2</sub>                              | 200 ppm                     | 300                                        | 8                     | 0.4                  |
|                                  |                                   | SiF <sub>4</sub>                            | 500                         |                                            |                       | 0.5                  |
|                                  | 4th layer region                  | AlCl <sub>3</sub> /He                       | 0.5                         |                                            |                       |                      |
|                                  |                                   | SiH <sub>4</sub>                            | 0.1                         |                                            |                       |                      |
|                                  |                                   | SiH <sub>4</sub>                            | 300                         |                                            |                       |                      |
| Upper layer                      | 2nd layer region                  | H <sub>2</sub>                              | 500                         |                                            |                       |                      |
|                                  |                                   | CH <sub>4</sub>                             | 1                           | 300                                        | 20                    | 0.5                  |
|                                  |                                   | NO                                          | 0.1                         |                                            |                       | 20                   |
|                                  | 3rd layer region                  | B <sub>2</sub> H <sub>6</sub>               | 0.3 ppm                     |                                            |                       |                      |
|                                  |                                   | SiF <sub>4</sub>                            | 0.5                         |                                            |                       |                      |
|                                  |                                   | AlCl <sub>3</sub> /He                       | 0.1                         |                                            |                       |                      |
| Lower layer                      | 4th layer region                  | SiH <sub>4</sub>                            | 100                         |                                            |                       |                      |
|                                  |                                   | CH <sub>4</sub>                             | 600                         |                                            |                       |                      |
|                                  |                                   | PH <sub>3</sub> (against SiH <sub>4</sub> ) | 3000 ppm                    | 300                                        | 15                    | 0.4                  |
|                                  | 5th layer region                  | NO                                          | 0.1                         |                                            |                       | 7                    |
|                                  |                                   | SiF <sub>4</sub>                            | 0.1                         |                                            |                       |                      |
|                                  |                                   | AlCl <sub>3</sub> /He                       | 0.1                         |                                            |                       |                      |

TABLE 95

| Order of lamination (layer name) | Gases and their flow rates (SCCM) |                                                           | Substrate temperature (°C.) | RF discharging power (mW/cm <sup>3</sup> ) | Inner pressure (Torr) | Layer thickness (μm) |
|----------------------------------|-----------------------------------|-----------------------------------------------------------|-----------------------------|--------------------------------------------|-----------------------|----------------------|
| Upper layer                      | 1st layer region                  | SiH <sub>4</sub>                                          | 10 → 100*                   |                                            |                       |                      |
|                                  |                                   | H <sub>2</sub>                                            | 5 → 200*                    |                                            |                       |                      |
|                                  |                                   | AlCl <sub>3</sub> /He (S-side: 0.05 μm)                   | 250                         | 5                                          | 0.4                   | 0.2                  |
|                                  | 2nd layer region                  | SiH <sub>4</sub>                                          | 200 → 40**                  |                                            |                       |                      |
|                                  |                                   | NO                                                        | 40 → 10**                   |                                            |                       |                      |
|                                  |                                   | SiH <sub>4</sub>                                          | 5 → 20                      |                                            |                       |                      |
| Lower layer                      | 3rd layer region                  | B <sub>2</sub> H <sub>6</sub> (against SiH <sub>4</sub> ) | 100                         |                                            |                       |                      |
|                                  |                                   | (LL-side: 2 μm)                                           |                             |                                            |                       |                      |
|                                  |                                   | (U + 2nd + LR-side: 1 μm)                                 | 500 ppm                     | 250                                        | 8                     | 0.4                  |
|                                  | 4th layer region                  | H <sub>2</sub>                                            | 500 ppm → 0**               |                                            |                       | 3                    |
|                                  |                                   | SiF <sub>4</sub>                                          | 200                         |                                            |                       |                      |
|                                  |                                   | AlCl <sub>3</sub> /He                                     | 0.5                         |                                            |                       |                      |
| Lower layer                      | SiH <sub>4</sub>                  | 0.1                                                       |                             |                                            |                       |                      |
|                                  | SiF <sub>4</sub>                  | 100                                                       |                             |                                            |                       |                      |

TABLE 95-continued

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| layer 1<br>layer region          | H <sub>2</sub>                                            | 200                         | 300                                        | 3                     | 0.5                  |
|                                  | CH <sub>4</sub>                                           | 1                           |                                            |                       | 3                    |
|                                  | NO                                                        | 0.1                         |                                            |                       |                      |
|                                  | B <sub>2</sub> H <sub>6</sub> (against SiH <sub>4</sub> ) | 0.3 ppm                     |                                            |                       |                      |
|                                  | AlCl <sub>3</sub> /He                                     | 0.1                         |                                            |                       |                      |
|                                  | SiH <sub>4</sub>                                          | 100                         |                                            |                       |                      |
|                                  | CH <sub>4</sub>                                           | 100                         |                                            |                       |                      |
|                                  | PH <sub>3</sub> (against SiH <sub>4</sub> )               | 50 ppm                      | 300                                        | 15                    | 0.4                  |
|                                  | NO                                                        | 0.1                         |                                            |                       | 30                   |
|                                  | B <sub>2</sub> H <sub>6</sub> (against SiH <sub>4</sub> ) | 0.3 ppm                     |                                            |                       |                      |
| layer 2<br>layer region          | SiF <sub>4</sub>                                          | 0.5                         |                                            |                       |                      |
|                                  | AlCl <sub>3</sub> /He                                     | 0.1                         |                                            |                       |                      |
|                                  | SiH <sub>4</sub>                                          | 50                          |                                            |                       |                      |
|                                  | CH <sub>4</sub>                                           | 600                         |                                            |                       |                      |
|                                  | PH <sub>3</sub> (against SiH <sub>4</sub> )               | 0.3 ppm                     | 300                                        | 10                    | 0.4                  |
| layer 3<br>layer region          | B <sub>2</sub> H <sub>6</sub> (against SiH <sub>4</sub> ) | 0.3 ppm                     |                                            |                       | 0.5                  |
|                                  | NO                                                        | 0.1                         |                                            |                       |                      |
|                                  | SiF <sub>4</sub>                                          | 0.5                         |                                            |                       |                      |
|                                  | AlCl <sub>3</sub> /He                                     | 0.1                         |                                            |                       |                      |

TABLE 96

| Order of lamination (layer name) | Gases and their flow rates (SCCM)            | Substrate temperature (°C.) | RF discharging power (mW/cm <sup>3</sup> ) | Inner pressure (Torr) | Layer thickness (μm) |
|----------------------------------|----------------------------------------------|-----------------------------|--------------------------------------------|-----------------------|----------------------|
| Lower layer                      | H <sub>2</sub> S (against SiH <sub>4</sub> ) | 1 ppm                       |                                            |                       |                      |
|                                  | SiH <sub>4</sub>                             | 10 → 100*                   |                                            |                       |                      |
|                                  | H <sub>2</sub>                               | 5 → 200*                    |                                            |                       |                      |
|                                  | AlCl <sub>3</sub> /He<br>(S-side: 0.05 μm)   | 300                         | 10                                         | 0.4                   | 0.2                  |
|                                  | 200 → 40**<br>(UL-side: 0.15 μm)             |                             |                                            |                       |                      |
|                                  | 40 → 10**                                    |                             |                                            |                       |                      |
|                                  | NO                                           | 5 → 20*                     |                                            |                       |                      |
|                                  | SiH <sub>4</sub>                             | 100                         |                                            |                       |                      |
|                                  | B <sub>2</sub> H <sub>6</sub>                | 200 ppm                     |                                            |                       |                      |
|                                  | H <sub>2</sub>                               | 500                         | 300                                        | 8                     | 0.4                  |
| Upper layer                      | SiF <sub>4</sub>                             | 0.5                         |                                            |                       | 0.5                  |
|                                  | AlCl <sub>3</sub> /He                        | 0.1                         |                                            |                       |                      |
|                                  | H <sub>2</sub> S                             | 1 ppm                       |                                            |                       |                      |
|                                  | SiH <sub>4</sub>                             | 300                         |                                            |                       |                      |
|                                  | H <sub>2</sub>                               | 500                         |                                            |                       |                      |
|                                  | CH <sub>4</sub>                              | 1                           | 300                                        | 20                    | 0.5                  |
|                                  | NO                                           | 0.1                         |                                            |                       | 20                   |
|                                  | B <sub>2</sub> H <sub>6</sub>                | 0.3 ppm                     |                                            |                       |                      |
|                                  | SiF <sub>4</sub>                             | 0.5                         |                                            |                       |                      |
|                                  | AlCl <sub>3</sub> /He                        | 0.1                         |                                            |                       |                      |
| 3rd layer                        | H <sub>2</sub> S                             | 1 ppm                       |                                            |                       |                      |
|                                  | SiH <sub>4</sub>                             | 100                         |                                            |                       |                      |
|                                  | CH <sub>4</sub>                              | 600                         |                                            |                       |                      |
|                                  | PH <sub>3</sub> (against SiH <sub>4</sub> )  | 3000 ppm                    | 300                                        | 15                    | 0.4                  |
|                                  | NO                                           | 0.1                         |                                            |                       | 7                    |
| 4th layer                        | SiF <sub>4</sub>                             | 0.5                         |                                            |                       |                      |
|                                  | AlCl <sub>3</sub> /He                        | 0.1                         |                                            |                       |                      |
|                                  | B <sub>2</sub> H <sub>6</sub>                | 0.3 ppm                     |                                            |                       |                      |
|                                  | H <sub>2</sub> S                             | 1 ppm                       |                                            |                       |                      |
|                                  | SiH <sub>4</sub>                             | 40                          |                                            |                       |                      |
|                                  | CH <sub>4</sub>                              | 600                         |                                            |                       |                      |
| region                           | NO                                           | 0.1                         | 300                                        | 10                    | 0.4                  |
|                                  | PH <sub>3</sub>                              | 0.3 ppm                     |                                            |                       | 0.1                  |
|                                  | B <sub>2</sub> H <sub>6</sub>                | 0.3 ppm                     |                                            |                       |                      |
|                                  | SiF <sub>4</sub>                             | 0.5                         |                                            |                       |                      |
|                                  | AlCl <sub>3</sub> /He                        | 0.1                         |                                            |                       |                      |
|                                  | H <sub>2</sub> S                             | 1 ppm                       |                                            |                       |                      |

TABLE 97

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 50                          |                                            |                       |                      |
|                                  | SiF <sub>4</sub>                                          | 5                           |                                            |                       |                      |
|                                  | H <sub>2</sub>                                            | 10 → 200*                   |                                            |                       |                      |
|                                  | AlCl <sub>3</sub> /He                                     | 120 → 40**                  |                                            |                       |                      |
|                                  | SiH <sub>4</sub>                                          | 100                         |                                            |                       |                      |
|                                  | B <sub>2</sub> H <sub>6</sub> (against SiH <sub>4</sub> ) | 200 ppm                     | 250                                        | 8                     | 0.4                  |
|                                  |                                                           |                             |                                            |                       | 3                    |
|                                  |                                                           |                             |                                            |                       |                      |
|                                  |                                                           |                             |                                            |                       |                      |
|                                  |                                                           |                             |                                            |                       |                      |
| 1st layer                        |                                                           |                             |                                            |                       |                      |
|                                  |                                                           |                             |                                            |                       |                      |
|                                  |                                                           |                             |                                            |                       |                      |
|                                  |                                                           |                             |                                            |                       |                      |
|                                  |                                                           |                             |                                            |                       |                      |

TABLE 97-continued

| Order of lamination (layer name) | Gases and their flow rates (SCCM) | Substrate temperature (°C.) | RF discharging power (mW/cm <sup>3</sup> ) | Inner pressure (Torr) | Layer thickness (μm) |
|----------------------------------|-----------------------------------|-----------------------------|--------------------------------------------|-----------------------|----------------------|
| Upper layer                      | H <sub>2</sub>                    | 250                         | 15                                         | 0.5                   | 20                   |
| 2nd layer                        | SiH <sub>4</sub>                  |                             |                                            |                       |                      |
| 2nd layer region                 | H <sub>2</sub>                    |                             |                                            |                       |                      |
| 3rd layer region                 | SiH <sub>4</sub>                  |                             |                                            |                       |                      |
| 3rd layer region                 | CH <sub>4</sub>                   |                             |                                            |                       |                      |

TABLE 98

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 250                         | 5                                          | 0.4                   | 0.05                 |
| 1st layer                        | AlCl <sub>3</sub> /He                                     |                             |                                            |                       |                      |
| 1st layer                        | SiH <sub>4</sub>                                          |                             |                                            |                       |                      |
| 1st layer region                 | B <sub>2</sub> H <sub>6</sub> (against SiH <sub>4</sub> ) |                             |                                            |                       |                      |
| Upper layer                      | H <sub>2</sub>                                            | 250                         | 8                                          | 0.4                   | 3                    |
| 2nd layer                        | SiH <sub>4</sub>                                          |                             |                                            |                       |                      |
| 2nd layer region                 | H <sub>2</sub>                                            |                             |                                            |                       |                      |
| 3rd layer region                 | SiH <sub>4</sub>                                          |                             |                                            |                       |                      |
| 3rd layer region                 | CH <sub>4</sub>                                           |                             |                                            |                       |                      |

TABLE 99

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiF <sub>4</sub>                                          | 250                         | 5                                          | 0.4                   | 0.03                 |
| 1st layer                        | SiH <sub>4</sub>                                          |                             |                                            |                       |                      |
| 1st layer                        | NO                                                        |                             |                                            |                       |                      |
| 1st layer                        | H <sub>2</sub>                                            |                             |                                            |                       |                      |
| Upper layer                      | AlCl <sub>3</sub> /He<br>(S-side: 0.01 μm)                | 250                         | 8                                          | 0.4                   | 3                    |
| 1st layer                        | 100 → 10**<br>(UL-side: 0.01 μm)                          |                             |                                            |                       |                      |
| 1st layer                        | 10                                                        |                             |                                            |                       |                      |
| 1st layer                        | B <sub>2</sub> H <sub>6</sub> (against SiH <sub>4</sub> ) |                             |                                            |                       |                      |
| 2nd layer                        | SiH <sub>4</sub>                                          | 250                         | 15                                         | 0.5                   | 20                   |
| 2nd layer                        | H <sub>2</sub>                                            |                             |                                            |                       |                      |
| 2nd layer                        | SiH <sub>4</sub>                                          |                             |                                            |                       |                      |
| 2nd layer                        | H <sub>2</sub>                                            |                             |                                            |                       |                      |
| 3rd layer                        | SiH <sub>4</sub>                                          | 250                         | 10                                         | 0.4                   | 0.5                  |
| 3rd layer                        | CH <sub>4</sub>                                           |                             |                                            |                       |                      |

TABLE 100

| Order of lamination (layer name) | Gases and their flow rates (SCCM)                                            | Substrate temperature (°C.) | RF discharging power (mW/cm <sup>3</sup> ) | Inner pressure (Torr) | Layer thickness (μm) |
|----------------------------------|------------------------------------------------------------------------------|-----------------------------|--------------------------------------------|-----------------------|----------------------|
| Lower layer                      | B <sub>2</sub> H <sub>6</sub> (against SiH <sub>4</sub> )                    | 150<br>300                  | 0.5<br>1.5                                 | 0.3                   | 0.02                 |
| 1st layer                        | SiF <sub>4</sub>                                                             |                             |                                            |                       |                      |
| 1st layer                        | SiH <sub>4</sub>                                                             |                             |                                            |                       |                      |
| 1st layer                        | H <sub>2</sub>                                                               |                             |                                            |                       |                      |
| Upper layer                      | AlCl <sub>3</sub> /He<br>(S-side: 0.01 μm)                                   | 250                         | 10                                         | 0.4                   | 3                    |
| 1st layer                        | 200 → 30**<br>(UL-side: 0.01 μm)                                             |                             |                                            |                       |                      |
| 1st layer                        | 30 → 10**                                                                    |                             |                                            |                       |                      |
| 1st layer                        | NO                                                                           |                             |                                            |                       |                      |
| 2nd layer                        | SiH <sub>4</sub>                                                             | 250                         | 20                                         | 0.5                   | 20                   |
| 2nd layer                        | B <sub>2</sub> H <sub>6</sub> (against SiH <sub>4</sub> )<br>(LL-side: 2 μm) |                             |                                            |                       |                      |
| 2nd layer                        | (U - 2nd - LR-side: 1 μm)                                                    |                             |                                            |                       |                      |
| 2nd layer                        | 500 ppm → 0**                                                                |                             |                                            |                       |                      |
| 2nd layer                        | H <sub>2</sub>                                                               | 250                         | 20                                         | 0.5                   | 20                   |
| 2nd layer                        | SiH <sub>4</sub>                                                             |                             |                                            |                       |                      |
| 2nd layer                        | H <sub>2</sub>                                                               |                             |                                            |                       |                      |

TABLE 101

| Order of lamination (layer name) | Gases and their flow rates (SCCM)                                                                                                                                                                                                                                                                                                                                                                                                    | Substrate temperature (°C.) | RF discharging power (mW/cm <sup>3</sup> ) | Inner pressure (Torr) | Layer thickness (μm) |
|----------------------------------|--------------------------------------------------------------------------------------------------------------------------------------------------------------------------------------------------------------------------------------------------------------------------------------------------------------------------------------------------------------------------------------------------------------------------------------|-----------------------------|--------------------------------------------|-----------------------|----------------------|
| Lower layer                      | SiH <sub>4</sub> 50<br>B <sub>2</sub> H <sub>6</sub> (against SiH <sub>4</sub> ) 100 ppm<br>SiF <sub>4</sub> 5<br>H <sub>2</sub> 5 → 200*<br>AlCl <sub>3</sub> /He (S-side: 0.01 μm)                                                                                                                                                                                                                                                 | 250                         | 1                                          | 0.3                   | 0.02                 |
|                                  | (UL-side: 0.01 μm) 200 → 30**<br>N <sub>2</sub> 100<br>SiH <sub>4</sub> 100<br>B <sub>2</sub> H <sub>6</sub> (against SiH <sub>4</sub> ) 500 ppm<br>He 600                                                                                                                                                                                                                                                                           | 250                         | 10                                         | 0.4                   | 3                    |
| Upper layer                      | AlCl <sub>3</sub> /He 0.1<br>SiF <sub>4</sub> 0.5<br>2nd layer region NO 0.1<br>CH <sub>4</sub> 1<br>SiH <sub>4</sub> 300<br>He 600<br>B <sub>2</sub> H <sub>6</sub> 0.3 ppm<br>SiF <sub>4</sub> 0.5<br>AlCl <sub>3</sub> /He 0.1<br>3rd layer region SiH <sub>4</sub> 50<br>CH <sub>4</sub> 500<br>NO 0.1<br>B <sub>2</sub> H <sub>6</sub> (against SiH <sub>4</sub> ) 0.3 ppm<br>SiF <sub>4</sub> 0.5<br>AlCl <sub>3</sub> /He 0.1 | 250                         | 25                                         | 0.6                   | 25                   |
|                                  |                                                                                                                                                                                                                                                                                                                                                                                                                                      | 250                         | 10                                         | 0.4                   | 1                    |

TABLE 102

| Order of lamination (layer name) | Gases and their flow rates (SCCM)                                                                                                                                                                                                                      | Substrate temperature (°C.) | RF discharging power (mW/cm <sup>3</sup> ) | Inner pressure (Torr) | Layer thickness (μm) |
|----------------------------------|--------------------------------------------------------------------------------------------------------------------------------------------------------------------------------------------------------------------------------------------------------|-----------------------------|--------------------------------------------|-----------------------|----------------------|
| Lower layer                      | SiH <sub>4</sub> 10 → 100*<br>H <sub>2</sub> 5 → 200*<br>Al(CH <sub>3</sub> ) <sub>3</sub> /He (S-side: 0.05 μm)                                                                                                                                       | 250                         | 10                                         | 0.4                   | 0.2                  |
|                                  | (UL-side: 0.15 μm) 200 → 40**<br>CH <sub>4</sub> 40 → 10**<br>SiF <sub>4</sub> 50 → 200*<br>1st layer region SiH <sub>4</sub> 100<br>B <sub>2</sub> H <sub>6</sub> (against SiH <sub>4</sub> ) 500 ppm<br>(LL-side: 2 μm)<br>(U + 2nd + LR-side: 1 μm) | 250                         | 10                                         | 0.4                   | 3                    |
| Upper layer                      | H <sub>2</sub> 200<br>SiH <sub>4</sub> 400<br>Ar 200<br>2nd layer region SiH <sub>4</sub> 100<br>NH <sub>3</sub> 30                                                                                                                                    | 250                         | 10                                         | 0.5                   | 15                   |
|                                  | 500 ppm → 0**<br>3rd layer region SiH <sub>4</sub> 100<br>NH <sub>3</sub> 30                                                                                                                                                                           | 250                         | 5                                          | 0.4                   | 0.3                  |

TABLE 103

| Order of lamination (layer name) | Gases and their flow rates (SCCM)                                                                                                                                                                             | Substrate temperature (°C.) | RF discharging power (mW/cm <sup>3</sup> ) | Inner pressure (Torr) | Layer thickness (μm) |
|----------------------------------|---------------------------------------------------------------------------------------------------------------------------------------------------------------------------------------------------------------|-----------------------------|--------------------------------------------|-----------------------|----------------------|
| Lower layer                      | SiH <sub>4</sub> 10 → 100*<br>H <sub>2</sub> 5 → 200*<br>AlCl <sub>3</sub> /He (S-side: 0.05 μm)                                                                                                              | 300                         | 10                                         | 0.4                   | 0.2                  |
|                                  | (UL-side: 0.15 μm) 200 → 40**<br>NO 40 → 10**<br>SiF <sub>4</sub> 5 → 20*<br>1st layer region SiH <sub>4</sub> 100<br>B <sub>2</sub> H <sub>6</sub> (against SiH <sub>4</sub> ) 200 ppm<br>H <sub>2</sub> 500 | 300                         | 8                                          | 0.4                   | 0.5                  |
| Upper layer                      | 2nd layer region SiH <sub>4</sub> 300<br>H <sub>2</sub> 500                                                                                                                                                   | 300                         | 20                                         | 0.5                   | 20                   |

TABLE 103-continued

| Order of lamination (layer name) | Gases and their flow rates (SCCM)                    | Substrate temperature (°C.) | RF discharging power (mW/cm <sup>3</sup> ) | Inner pressure (Torr) | Layer thickness (μm) |
|----------------------------------|------------------------------------------------------|-----------------------------|--------------------------------------------|-----------------------|----------------------|
| 3rd layer region                 | SiH <sub>4</sub> 100                                 | 300                         | 15                                         | 0.4                   | 7                    |
|                                  | CH <sub>4</sub> 600                                  |                             |                                            |                       |                      |
|                                  | PH <sub>3</sub> (against SiH <sub>4</sub> ) 3000 ppm |                             |                                            |                       |                      |
| 4th layer region                 | SiH <sub>4</sub> 40                                  | 300                         | 10                                         | 0.4                   | 0.1                  |
|                                  | CH <sub>4</sub> 600                                  |                             |                                            |                       |                      |

TABLE 104

| Order of lamination (layer name) | Gases and their flow rates (SCCM)                                  | Substrate temperature (°C.) | RF discharging power (mW/cm <sup>3</sup> ) | Inner pressure (Torr) | Layer thickness (μm) |
|----------------------------------|--------------------------------------------------------------------|-----------------------------|--------------------------------------------|-----------------------|----------------------|
| Lower layer                      | PF <sub>3</sub> (against SiH <sub>4</sub> ) 50 ppm                 | 330                         | 5                                          | 0.4                   | 0.05                 |
|                                  | SiH <sub>4</sub> 50                                                |                             |                                            |                       |                      |
|                                  | H <sub>2</sub> 5 → 200*                                            |                             |                                            |                       |                      |
|                                  | AlCl <sub>3</sub> /He 200 → 20**                                   |                             |                                            |                       |                      |
|                                  | NO 5                                                               |                             |                                            |                       |                      |
|                                  | SiF <sub>4</sub> 5                                                 |                             |                                            |                       |                      |
| Upper layer                      | 1st layer region SiH <sub>4</sub> 100                              | 330                         | 8                                          | 0.4                   | 3                    |
|                                  | PH <sub>3</sub> 100 ppm                                            |                             |                                            |                       |                      |
|                                  | H <sub>2</sub> 100                                                 |                             |                                            |                       |                      |
|                                  | 2nd layer region SiH <sub>4</sub> 400                              |                             |                                            |                       |                      |
|                                  | SiF <sub>4</sub> 10                                                |                             |                                            |                       |                      |
|                                  | H <sub>2</sub> 800                                                 |                             |                                            |                       |                      |
| 4th layer region                 | 3rd layer region SiH <sub>4</sub> 100                              | 350                         | 15                                         | 0.4                   | 5                    |
|                                  | CH <sub>4</sub> 400                                                |                             |                                            |                       |                      |
|                                  | B <sub>2</sub> H <sub>6</sub> (against SiH <sub>4</sub> ) 5000 ppm |                             |                                            |                       |                      |
|                                  | SiH <sub>4</sub> 20                                                |                             |                                            |                       |                      |
|                                  | CH <sub>4</sub> 400                                                |                             |                                            |                       |                      |
|                                  | B <sub>2</sub> H <sub>6</sub> (against SiH <sub>4</sub> ) 8000 ppm |                             |                                            |                       |                      |

TABLE 105

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 50                                               | 300                         | 1                                          | 0.3                   | 0.02                 |
|                                  | H <sub>2</sub> S (against SiH <sub>4</sub> ) 10 ppm               |                             |                                            |                       |                      |
|                                  | SiF <sub>4</sub> 5                                                |                             |                                            |                       |                      |
|                                  | H <sub>2</sub> 5 → 200*                                           |                             |                                            |                       |                      |
|                                  | AlCl <sub>3</sub> /He (S-side: 0.01 μm) 200 → 30**                |                             |                                            |                       |                      |
|                                  | (UL-side: 0.01 μm) 30 → 10**                                      |                             |                                            |                       |                      |
| Upper layer                      | 1st layer region SiH <sub>4</sub> 100                             | 300                         | 8                                          | 0.4                   | 5                    |
|                                  | B <sub>2</sub> H <sub>6</sub> (against SiH <sub>4</sub> ) 200 ppm |                             |                                            |                       |                      |
|                                  | H <sub>2</sub> 200                                                |                             |                                            |                       |                      |
|                                  | 2nd layer region SiH <sub>4</sub> 300                             |                             |                                            |                       |                      |
|                                  | H <sub>2</sub> 200                                                |                             |                                            |                       |                      |
|                                  | 3rd layer region SiH <sub>4</sub> 50                              |                             |                                            |                       |                      |
| 4th layer region                 | N <sub>2</sub> 500                                                | 300                         | 20                                         | 0.4                   | 5                    |
|                                  | PH <sub>3</sub> (against SiH <sub>4</sub> ) 3000 ppm              |                             |                                            |                       |                      |
|                                  | SiH <sub>4</sub> 40                                               |                             |                                            |                       |                      |
|                                  | CH <sub>4</sub> 600                                               |                             |                                            |                       |                      |

TABLE 106

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | B <sub>2</sub> H <sub>6</sub> (against SiH <sub>4</sub> ) 100 ppm | 250                         | 5                                          | 0.4                   | 0.05                 |
|                                  | SiH <sub>4</sub> 50                                               |                             |                                            |                       |                      |
|                                  | H <sub>2</sub> 5 → 200*                                           |                             |                                            |                       |                      |
|                                  | AlCl <sub>3</sub> /He 200 → 20**                                  |                             |                                            |                       |                      |
|                                  | NO 5                                                              |                             |                                            |                       |                      |
|                                  | C <sub>2</sub> H <sub>2</sub> 10                                  |                             |                                            |                       |                      |
|                                  | SiF <sub>4</sub> 5                                                |                             |                                            |                       |                      |

TABLE 106-continued

| Order of lamination (layer name) | Gases and their flow rates (SCCM) |                                                                                                                               | Substrate temperature (°C.)     | RF discharging power (mW/cm <sup>3</sup> ) | Inner pressure (Torr) | Layer thickness (μm) |
|----------------------------------|-----------------------------------|-------------------------------------------------------------------------------------------------------------------------------|---------------------------------|--------------------------------------------|-----------------------|----------------------|
| Upper layer                      | 1st layer                         | SiH <sub>4</sub><br>B <sub>2</sub> H <sub>6</sub> (against SiH <sub>4</sub> )<br>(LL-side: 3 μm)<br>(U · 2nd · LR-side: 2 μm) | 100<br>500 ppm<br>500 ppm → 0** | 250                                        | 10                    | 0.4                  |
|                                  | 2nd layer                         | H <sub>2</sub><br>AlCl <sub>3</sub> /He (against SiH <sub>4</sub> )                                                           | 200<br>1 → 0**                  | 250                                        | 15                    | 0.5                  |
|                                  | 3rd layer                         | SiH <sub>4</sub><br>C <sub>2</sub> H <sub>2</sub>                                                                             | 300<br>200                      | 250                                        | 15                    | 10                   |
|                                  | region                            | NO                                                                                                                            | 10 → 20*                        | 250                                        | 0.4                   | 20                   |
|                                  |                                   |                                                                                                                               | 1                               |                                            |                       |                      |

TABLE 107

| Order of lamination (layer name) | Gases and their flow rates (SCCM)                                            |               | Substrate temperature (°C.) | RF discharging power (mW/cm <sup>3</sup> ) | Inner pressure (Torr) | Layer thickness (μm) |
|----------------------------------|------------------------------------------------------------------------------|---------------|-----------------------------|--------------------------------------------|-----------------------|----------------------|
| Lower layer                      | NO                                                                           | 1             |                             |                                            |                       |                      |
|                                  | SiH <sub>4</sub>                                                             | 50            |                             |                                            |                       |                      |
|                                  | H <sub>2</sub>                                                               | 5 → 200*      |                             |                                            |                       |                      |
|                                  | AlCl <sub>3</sub> /He<br>(S-side: 0.01 μm)                                   | 200 → 30**    | 250                         | 1                                          | 0.4                   | 0.02                 |
| Upper layer                      | (UL-side: 0.01 μm)                                                           |               |                             |                                            |                       |                      |
|                                  | BF <sub>3</sub> (against SiH <sub>4</sub> )                                  | 30 → 10**     |                             |                                            |                       |                      |
| Upper layer                      | SiF <sub>4</sub>                                                             | 100           |                             |                                            |                       |                      |
|                                  | SiH <sub>4</sub>                                                             | 5             |                             |                                            |                       |                      |
|                                  | B <sub>2</sub> H <sub>6</sub> (against SiH <sub>4</sub> )<br>(LL-side: 2 μm) | 500 ppm       | 250                         | 10                                         | 0.4                   | 10                   |
|                                  | (U · 2nd · LR-side: 1 μm)                                                    | 500 ppm → 0** |                             |                                            |                       |                      |
| Upper layer                      | H <sub>2</sub>                                                               | 200           |                             |                                            |                       |                      |
|                                  | SiH <sub>4</sub>                                                             | 300           |                             |                                            |                       |                      |
| Upper layer                      | H <sub>2</sub>                                                               | 300           | 300                         | 20                                         | 0.5                   | 5                    |
|                                  | SiH <sub>4</sub>                                                             | 100           | 300                         | 15                                         | 0.4                   | 20                   |
| Upper layer                      | CH <sub>4</sub>                                                              | 100           |                             |                                            |                       |                      |
|                                  | SiH <sub>4</sub>                                                             | 50            | 300                         | 10                                         | 0.4                   | 0.5                  |
|                                  | CH <sub>4</sub>                                                              | 600           |                             |                                            |                       |                      |

TABLE 108

| Order of lamination (layer name) | Gases and their flow rates (SCCM)                         |            | Substrate temperature (°C.) | RF discharging power (mW/cm <sup>3</sup> ) | Inner pressure (Torr) | Layer thickness (μm) |
|----------------------------------|-----------------------------------------------------------|------------|-----------------------------|--------------------------------------------|-----------------------|----------------------|
| Lower layer                      | SiH <sub>4</sub>                                          | 10 → 100*  |                             |                                            |                       |                      |
|                                  | H <sub>2</sub>                                            | 5 → 200*   |                             |                                            |                       |                      |
|                                  | AlCl <sub>3</sub> /He<br>(S-side: 0.05 μm)                | 200 → 40** | 300                         | 5                                          | 0.4                   | 0.2                  |
|                                  | (UL-side: 0.15 μm)                                        | 40 → 10**  |                             |                                            |                       |                      |
| Upper layer                      | NH <sub>3</sub>                                           | 5 → 50*    |                             |                                            |                       |                      |
|                                  | SiF <sub>4</sub>                                          | 1 → 10*    |                             |                                            |                       |                      |
|                                  | SiH <sub>4</sub>                                          | 100        |                             |                                            |                       |                      |
|                                  | B <sub>2</sub> H <sub>6</sub> (against SiH <sub>4</sub> ) | 200 ppm    | 300                         | 5                                          | 0.4                   | 3                    |
| Upper layer                      | H <sub>2</sub>                                            | 500        |                             |                                            |                       |                      |
|                                  | SiH <sub>4</sub>                                          | 100        | 300                         | 5                                          | 0.2                   | 25                   |
| Upper layer                      | H <sub>2</sub>                                            | 300        | 300                         | 15                                         | 0.4                   | 25                   |
|                                  | NH <sub>3</sub>                                           | 50         | 300                         | 10                                         | 0.4                   | 0.3                  |
| Upper layer                      | SiH <sub>4</sub>                                          | 100        |                             |                                            |                       |                      |
|                                  | NH <sub>4</sub>                                           | 50         | 300                         | 10                                         | 0.4                   | 0.3                  |

TABLE 109

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 10 → 100*                   |                                            |                       |                      |
|                                  | H <sub>2</sub>                                            | 5 → 200*                    |                                            |                       |                      |
|                                  | AlCl <sub>3</sub> /He<br>(S-side: 0.05 μm)                |                             |                                            |                       |                      |
|                                  | (UL-side: 0.15 μm)                                        | 200 → 40**                  | 250                                        | 5                     | 0.4                  |
|                                  | NO                                                        | 40 → 10**                   |                                            |                       |                      |
|                                  | B <sub>2</sub> H <sub>6</sub> (against SiH <sub>4</sub> ) | 5 → 20*                     |                                            |                       |                      |
|                                  | SiF <sub>4</sub>                                          | 100 ppm                     |                                            |                       |                      |
|                                  | SiH <sub>4</sub>                                          | 1 → 10*                     |                                            |                       |                      |
|                                  | B <sub>2</sub> H <sub>6</sub> (against SiH <sub>4</sub> ) | 100                         |                                            |                       |                      |
|                                  | (LL-side: 2 μm)<br>(U · 2nd · LR-side: 1 μm)              | 500 ppm                     | 250                                        | 8                     | 0.4                  |
| Upper layer region               |                                                           | 500 ppm → 0**               |                                            |                       | 3                    |
|                                  | H <sub>2</sub>                                            | 200                         |                                            |                       |                      |
|                                  | Si <sub>2</sub> F <sub>6</sub>                            | 5                           |                                            |                       |                      |
|                                  | SiH <sub>4</sub>                                          | 100                         |                                            |                       |                      |
|                                  | SiF <sub>4</sub>                                          | 5                           | 300                                        | 3                     | 0.5                  |
|                                  | H <sub>2</sub>                                            | 200                         |                                            |                       |                      |
|                                  | SiH <sub>4</sub>                                          | 100                         |                                            |                       |                      |
|                                  | CH <sub>4</sub>                                           | 100                         | 300                                        | 15                    | 0.4                  |
|                                  | PH <sub>3</sub> (against SiH <sub>4</sub> )               | 50 ppm                      |                                            |                       | 30                   |
|                                  | SiH <sub>4</sub>                                          | 50                          |                                            |                       |                      |
| 3rd layer region                 | CH <sub>4</sub>                                           | 600                         | 300                                        | 10                    | 0.4                  |
|                                  |                                                           |                             |                                            |                       | 0.5                  |
| 4th layer region                 |                                                           |                             |                                            |                       |                      |

TABLE 110

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | N <sub>2</sub>                                            | 300                         |                                            |                       |                      |
|                                  | SiH <sub>4</sub>                                          | 50                          |                                            |                       |                      |
|                                  | H <sub>2</sub>                                            | 5 → 200*                    | 250                                        | 5                     | 0.4                  |
|                                  | AlCl <sub>3</sub> /He                                     | 200 → 20**                  |                                            |                       |                      |
|                                  | PH <sub>3</sub> (against SiH <sub>4</sub> )               | 50 ppm                      |                                            |                       |                      |
|                                  | Si <sub>2</sub> F <sub>6</sub>                            | 5                           |                                            |                       |                      |
|                                  | SiH <sub>4</sub>                                          | 40                          | *                                          |                       |                      |
|                                  | PH <sub>3</sub> (against SiH <sub>4</sub> )               | 250 ppm                     | 250                                        | 8                     | 0.4                  |
|                                  | (LL-side: 2 μm)<br>(U · 2nd · LR-side: 1 μm)              | 250 ppm → 0**               |                                            |                       | 3                    |
|                                  | H <sub>2</sub>                                            | 40                          |                                            |                       |                      |
| Upper layer region               | Si <sub>2</sub> H <sub>6</sub>                            | 200                         |                                            |                       |                      |
|                                  | H <sub>2</sub>                                            | 200                         | 300                                        | 10                    | 0.5                  |
|                                  | SiH <sub>4</sub>                                          | 300                         |                                            |                       |                      |
|                                  | C <sub>2</sub> H <sub>2</sub>                             | 50                          |                                            |                       |                      |
|                                  | B <sub>2</sub> H <sub>6</sub> (against SiH <sub>4</sub> ) | 0 → 100 ppm*                | 330                                        | 20                    | 0.4                  |
|                                  | (U · 2nd · LR-side: 1 μm)                                 | (U · 4th · LR-side: 29 μm)  |                                            |                       | 30                   |
|                                  | SiH <sub>4</sub>                                          | 100 ppm                     |                                            |                       |                      |
|                                  | C <sub>2</sub> H <sub>2</sub>                             | 200                         | 330                                        | 10                    | 0.4                  |
|                                  |                                                           | 200                         |                                            |                       | 1                    |

TABLE 111

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | B <sub>2</sub> H <sub>6</sub> (against SiH <sub>4</sub> ) | 80 ppm                      |                                            |                       |                      |
|                                  | SiH <sub>4</sub>                                          | 10 → 100*                   |                                            |                       |                      |
|                                  | H <sub>2</sub>                                            | 5 → 200*                    |                                            |                       |                      |
|                                  | AlCl <sub>3</sub> /He<br>(S-side: 0.05 μm)                |                             |                                            |                       |                      |
|                                  | (UL-side: 0.15 μm)                                        | 200 → 40**                  | 250                                        | 5                     | 0.4                  |
|                                  | NO                                                        | 40 → 10**                   |                                            |                       |                      |
|                                  | Si <sub>2</sub> F <sub>6</sub>                            | 5 → 20*                     |                                            |                       |                      |
|                                  | SiH <sub>4</sub>                                          | 1 → 10*                     |                                            |                       |                      |
|                                  | B <sub>2</sub> H <sub>6</sub> (against SiH <sub>4</sub> ) | 100                         |                                            |                       |                      |
|                                  | H <sub>2</sub>                                            | 200 ppm                     | 300                                        | 8                     | 0.3                  |
| 1st layer region                 |                                                           | 500                         |                                            |                       | 3                    |

TABLE 111-continued

| Order of lamination (layer name) | Gases and their flow rates (SCCM)                                          | Substrate temperature (°C.) | RF discharging power (mW/cm <sup>3</sup> ) | Inner pressure (Torr) | Layer thickness (μm) |
|----------------------------------|----------------------------------------------------------------------------|-----------------------------|--------------------------------------------|-----------------------|----------------------|
| 2nd layer region                 | SiH <sub>4</sub> 100<br>H <sub>2</sub> 300                                 | 300                         | 5                                          | 0.5                   | 8                    |
| 3rd layer region                 | SiH <sub>4</sub> 300<br>NH <sub>3</sub> 30 → 50*                           | 300                         | 15                                         | 0.4                   | 25                   |
| 4th layer region                 | PH <sub>3</sub> (against SiH <sub>4</sub> ) 50 ppm<br>SiH <sub>4</sub> 100 | 300                         | 5                                          | 0.4                   | 0.7                  |
|                                  | NH <sub>3</sub> 80 → 100*                                                  | 300                         | 5                                          | 0.4                   | 0.7                  |
|                                  | PH <sub>3</sub> (against SiH <sub>4</sub> ) 500 ppm                        |                             |                                            |                       |                      |

TABLE 112

| Order of lamination (layer name) | Gases and their flow rates (SCCM)                                          | Substrate temperature (°C.) | RF discharging power (mW/cm <sup>3</sup> ) | Inner pressure (Torr) | Layer thickness (μm) |
|----------------------------------|----------------------------------------------------------------------------|-----------------------------|--------------------------------------------|-----------------------|----------------------|
| Lower layer                      | SiH <sub>4</sub> 50<br>H <sub>2</sub> 5 → 200*                             |                             |                                            |                       |                      |
|                                  | AlCl <sub>3</sub> /He (S-side: 0.01 μm)                                    | 200 → 30**                  | 250                                        | 1                     | 0.4                  |
|                                  | (UL-side: 0.01 μm)                                                         | 30 → 10**                   |                                            |                       |                      |
|                                  | NO 10                                                                      |                             |                                            |                       |                      |
|                                  | SiF <sub>4</sub> 5                                                         |                             |                                            |                       |                      |
| Upper layer                      | 1st layer region SiH <sub>4</sub> 100<br>PH <sub>3</sub> 100 ppm           | 300                         | 8                                          | 0.4                   | 3                    |
|                                  | 2nd layer region SiH <sub>4</sub> 300<br>H <sub>2</sub> 500                | 300                         | 20                                         | 0.5                   | 20                   |
|                                  | 3rd layer region SiH <sub>4</sub> 100<br>GeH <sub>4</sub> 10 → 50*         | 300                         | 5                                          | 0.4                   | 1                    |
|                                  | 2nd layer region H <sub>2</sub> 300                                        |                             |                                            |                       |                      |
|                                  | 4th layer region SiH <sub>4</sub> 100 → 40**<br>CH <sub>4</sub> 100 → 600* | 300                         | 10                                         | 0.4                   | 1                    |

TABLE 113

| Order of lamination (layer name) | Gases and their flow rates (SCCM)                                                                                  | Substrate temperature (°C.) | RF discharging power (mW/cm <sup>3</sup> ) | Inner pressure (Torr) | Layer thickness (μm) |
|----------------------------------|--------------------------------------------------------------------------------------------------------------------|-----------------------------|--------------------------------------------|-----------------------|----------------------|
| Lower layer                      | B <sub>2</sub> H <sub>6</sub> (against SiH <sub>4</sub> ) 50 ppm<br>SiH <sub>4</sub> 50<br>H <sub>2</sub> 5 → 200* |                             |                                            |                       |                      |
|                                  | AlCl <sub>3</sub> /He (S-side: 0.01 μm)                                                                            | 200 → 30**                  | 300                                        | 1                     | 0.3                  |
|                                  | (UL-side: 0.01 μm)                                                                                                 | 30 → 10**                   |                                            |                       |                      |
|                                  | NO 5                                                                                                               |                             |                                            |                       |                      |
|                                  | SiF <sub>4</sub> 5                                                                                                 |                             |                                            |                       |                      |
| Upper layer                      | 1st layer region B <sub>2</sub> H <sub>6</sub> (against SiH <sub>4</sub> ) 200 ppm<br>H <sub>2</sub> 500           | 300                         | 8                                          | 0.4                   | 10                   |
|                                  | 2nd layer region SiH <sub>4</sub> 300<br>H <sub>2</sub> 400                                                        | 300                         | 15                                         | 0.5                   | 20                   |
|                                  | 3rd layer region SiH <sub>4</sub> 50<br>CH <sub>4</sub> 500                                                        | 300                         | 10                                         | 0.4                   | 0.5                  |

TABLE 114

| Order of lamination (layer name) | Gases and their flow rates (SCCM)                                                                                          | Substrate temperature (°C.) | RF discharging power (mW/cm <sup>3</sup> ) | Inner pressure (Torr) | Layer thickness (μm) |
|----------------------------------|----------------------------------------------------------------------------------------------------------------------------|-----------------------------|--------------------------------------------|-----------------------|----------------------|
| Lower layer                      | SiH <sub>4</sub> 50<br>B <sub>2</sub> H <sub>6</sub> (against SiH <sub>4</sub> ) 50 ppm<br>NO 5<br>H <sub>2</sub> 5 → 200* |                             |                                            |                       |                      |
|                                  | AlCl <sub>3</sub> /He (S-side: 0.01 μm)                                                                                    | 300                         | 0.7                                        | 0.3                   | 0.02                 |
|                                  | 200 → 30**                                                                                                                 |                             |                                            |                       |                      |

TABLE 114-continued

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| (UL-side: 0.01 μm)               |                                                           |                             |                                            |                       |                      |
| Upper layer                      | SiF <sub>4</sub>                                          | 30 → 10**                   |                                            |                       |                      |
|                                  | SiH <sub>4</sub>                                          | 5                           |                                            |                       |                      |
|                                  | H <sub>2</sub>                                            | 80                          |                                            |                       |                      |
|                                  | B <sub>2</sub> H <sub>6</sub> (against SiH <sub>4</sub> ) | 400                         | 300                                        | 7                     | 0.3                  |
|                                  |                                                           | 200 ppm                     |                                            |                       |                      |
|                                  | SiH <sub>4</sub>                                          | 200                         |                                            |                       |                      |
| 2nd layer region                 | H <sub>2</sub>                                            | 400                         | 300                                        | 12                    | 0.4                  |
|                                  | SiH <sub>4</sub>                                          | 40                          |                                            |                       |                      |
|                                  | CH <sub>4</sub>                                           | 400                         | 300                                        | 7                     | 0.3                  |
| 3rd layer region                 |                                                           |                             |                                            |                       | 0.5                  |

TABLE 115

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| (UL-side: 0.01 μm)               |                                                           |                             |                                            |                       |                      |
| Lower layer                      | SiH <sub>4</sub>                                          | 25                          |                                            |                       |                      |
|                                  | B <sub>2</sub> H <sub>6</sub> (against SiH <sub>4</sub> ) | 50 ppm                      |                                            |                       |                      |
|                                  | NO                                                        | 3                           |                                            |                       |                      |
|                                  | H <sub>2</sub>                                            | 5 → 100*                    |                                            |                       |                      |
|                                  | AlCl <sub>3</sub> /He                                     |                             | 300                                        | 0.5                   | 0.2                  |
|                                  | (S-side: 0.01 μm)                                         |                             | 100 → 15**                                 |                       |                      |
| (UL-side: 0.01 μm)               |                                                           |                             |                                            |                       |                      |
| Upper layer                      | SiF <sub>4</sub>                                          | 15 → 5**                    |                                            |                       |                      |
|                                  | SiH <sub>4</sub>                                          | 5                           |                                            |                       |                      |
|                                  | H <sub>2</sub>                                            | 60                          |                                            |                       |                      |
|                                  | B <sub>2</sub> H <sub>6</sub> (against SiH <sub>4</sub> ) | 300                         | 300                                        | 6                     | 0.2                  |
|                                  | SiH <sub>4</sub>                                          | 200 ppm                     |                                            |                       |                      |
|                                  | H <sub>2</sub>                                            | 150                         |                                            |                       |                      |
| 2nd layer region                 | SiH <sub>4</sub>                                          | 300                         | 300                                        | 10                    | 0.4                  |
|                                  | H <sub>2</sub>                                            | 300                         |                                            |                       |                      |
|                                  | SiH <sub>4</sub>                                          |                             |                                            |                       | 20                   |
| 3rd layer region                 | SiH <sub>4</sub>                                          | 30                          |                                            |                       |                      |
|                                  | CH <sub>4</sub>                                           | 300                         | 300                                        | 5                     | 0.3                  |
| region                           |                                                           |                             |                                            |                       | 0.5                  |

TABLE 116

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| (UL-side: 0.01 μm)               |                                                           |                             |                                            |                       |                      |
| Lower layer                      | SiH <sub>4</sub>                                          | 20                          |                                            |                       |                      |
|                                  | B <sub>2</sub> H <sub>6</sub> (against SiH <sub>4</sub> ) | 50 ppm                      |                                            |                       |                      |
|                                  | NO                                                        | 2                           |                                            |                       |                      |
|                                  | H <sub>2</sub>                                            | 5 → 100*                    |                                            |                       |                      |
|                                  | AlCl <sub>3</sub> /He                                     |                             | 300                                        | 0.3                   | 0.2                  |
|                                  | (S-side: 0.01 μm)                                         |                             | 80 → 15**                                  |                       |                      |
| (UL-side: 0.01 μm)               |                                                           |                             |                                            |                       |                      |
| Upper layer                      | SiF <sub>4</sub>                                          | 15 → 5**                    |                                            |                       |                      |
|                                  | SiH <sub>4</sub>                                          | 5                           |                                            |                       |                      |
|                                  | H <sub>2</sub>                                            | 40                          |                                            |                       |                      |
|                                  | B <sub>2</sub> H <sub>6</sub> (against SiH <sub>4</sub> ) | 200 ppm                     | 300                                        | 5                     | 0.2                  |
|                                  | SiH <sub>4</sub>                                          | 200                         |                                            |                       |                      |
|                                  | H <sub>2</sub>                                            | 100                         |                                            |                       |                      |
| 2nd layer region                 | SiH <sub>4</sub>                                          | 300                         | 300                                        | 6                     | 0.3                  |
|                                  | H <sub>2</sub>                                            | 300                         |                                            |                       |                      |
|                                  | SiH <sub>4</sub>                                          |                             |                                            |                       | 20                   |
| 3rd layer region                 | SiH <sub>4</sub>                                          | 20                          |                                            |                       |                      |
|                                  | CH <sub>4</sub>                                           | 200                         | 300                                        | 3                     | 0.2                  |
| region                           |                                                           |                             |                                            |                       | 0.5                  |

TABLE 117

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 50                          |                                            |                       |                      |
|                                  | B <sub>2</sub> H <sub>6</sub> (against SiH <sub>4</sub> ) | 100 ppm                     |                                            |                       |                      |
|                                  | NO                                                        | 5                           |                                            |                       |                      |
|                                  | H <sub>2</sub>                                            | 5 → 200*                    |                                            |                       |                      |
|                                  | AlCl <sub>3</sub> /He                                     | 200 → 20**                  |                                            |                       |                      |
|                                  | SiF <sub>4</sub>                                          | 5                           |                                            |                       |                      |

TABLE 117-continued

| Order of lamination (layer name) | Gases and their flow rates (SCCM) |                                                                              | Substrate temperature (°C.) | RF discharging power (mW/cm <sup>3</sup> ) | Inner pressure (Torr) | Layer thickness (μm) |
|----------------------------------|-----------------------------------|------------------------------------------------------------------------------|-----------------------------|--------------------------------------------|-----------------------|----------------------|
| Upper layer region               | 1st layer                         | SiH <sub>4</sub>                                                             | 100                         |                                            |                       |                      |
|                                  |                                   | B <sub>2</sub> H <sub>6</sub> (against SiH <sub>4</sub> )<br>(LL-side: 2 μm) | 500 ppm                     | 500                                        | 20                    | 0.4                  |
|                                  |                                   | U · 2nd · LR-side: 1 μm                                                      | 500 → 0 ppm**               |                                            |                       |                      |
| 2nd layer region                 | SiH <sub>4</sub>                  | H <sub>2</sub>                                                               | 1200                        |                                            |                       |                      |
|                                  |                                   |                                                                              | 300                         |                                            |                       |                      |
| 3rd layer region                 | SiH <sub>4</sub>                  | H <sub>2</sub>                                                               | 1500                        | 500                                        | 30                    | 0.5                  |
|                                  |                                   |                                                                              | 200                         |                                            |                       |                      |
|                                  | C <sub>2</sub> H <sub>2</sub>     | NO                                                                           | 10 → 20*                    | 500                                        | 30                    | 0.4                  |
|                                  |                                   |                                                                              | 1                           |                                            |                       | 20                   |

TABLE 118

| Order of lamination (layer name) | Gases and their flow rates (SCCM)                         |                                                           | Substrate temperature (°C.) | μW discharging power (mW/cm <sup>3</sup> ) | Inner pressure (Torr) | Layer thickness (μm) |
|----------------------------------|-----------------------------------------------------------|-----------------------------------------------------------|-----------------------------|--------------------------------------------|-----------------------|----------------------|
| Lower layer                      | B <sub>2</sub> H <sub>6</sub> (against SiH <sub>4</sub> ) | 50 ppm                                                    |                             |                                            |                       |                      |
|                                  | SiH <sub>4</sub>                                          | 150                                                       |                             |                                            |                       |                      |
|                                  | H <sub>2</sub>                                            | 20 → 500*                                                 |                             |                                            |                       |                      |
|                                  | AlCl <sub>3</sub> /He<br>(S-side: 0.01 μm)                | 400 → 80**                                                | 250                         | 0.5                                        | 0.6                   | 0.02                 |
|                                  | (UL-side: 0.01 μm)                                        | 80 → 50**                                                 |                             |                                            |                       |                      |
|                                  | NO                                                        | 10                                                        |                             |                                            |                       |                      |
| Upper Layer                      | SiF <sub>4</sub>                                          | 10                                                        |                             |                                            |                       |                      |
|                                  | 1st layer                                                 | SiH <sub>4</sub>                                          | 100                         |                                            |                       |                      |
|                                  |                                                           | B <sub>2</sub> H <sub>6</sub> (against SiH <sub>4</sub> ) | 200 ppm                     | 0.5                                        | 0.5                   | 3                    |
|                                  |                                                           | H <sub>2</sub>                                            | 500                         |                                            |                       |                      |
|                                  | 2nd layer                                                 | SiH <sub>4</sub>                                          | 700                         |                                            |                       |                      |
|                                  |                                                           | SiF <sub>4</sub>                                          | 30                          | 0.5                                        | 0.5                   | 20                   |
| 3rd layer                        | H <sub>2</sub>                                            | 500                                                       |                             |                                            |                       |                      |
|                                  | SiH <sub>4</sub>                                          | 150                                                       |                             |                                            |                       |                      |
|                                  | CH <sub>4</sub>                                           | 500                                                       | 250                         | 0.5                                        | 0.3                   | 1                    |
|                                  |                                                           |                                                           |                             |                                            |                       |                      |

TABLE 119

| Order of lamination (layer name) | Gases and their flow rates (SCCM)                         |                                                           | Substrate temperature (°C.) | RF discharging power (mW/cm <sup>3</sup> ) | Inner pressure (Torr) | Layer thickness (μm) |
|----------------------------------|-----------------------------------------------------------|-----------------------------------------------------------|-----------------------------|--------------------------------------------|-----------------------|----------------------|
| Lower layer                      | B <sub>2</sub> H <sub>6</sub> (against SiH <sub>4</sub> ) | 100 ppm                                                   |                             |                                            |                       |                      |
|                                  | SiH <sub>4</sub>                                          | 50                                                        |                             |                                            |                       |                      |
|                                  | H <sub>2</sub>                                            | 5 → 200*                                                  | 250                         | 5                                          | 0.4                   | 0.05                 |
|                                  | AlCl <sub>3</sub> /He                                     | 200 → 20**                                                |                             |                                            |                       |                      |
|                                  | NO                                                        | 5                                                         |                             |                                            |                       |                      |
|                                  | C <sub>2</sub> H <sub>2</sub>                             | 10                                                        |                             |                                            |                       |                      |
| Upper layer                      | SiF <sub>4</sub>                                          | 5                                                         |                             |                                            |                       |                      |
|                                  | 1st layer                                                 | SiH <sub>4</sub>                                          | 100                         |                                            |                       |                      |
|                                  |                                                           | B <sub>2</sub> H <sub>6</sub> (against SiH <sub>4</sub> ) |                             |                                            |                       |                      |
|                                  |                                                           | (LL-side: 3 μm)                                           | 500 ppm                     |                                            |                       |                      |
|                                  |                                                           | (U · 2nd · LR-side: 2 μm)                                 | 500 ppm → 0**               | 250                                        | 10                    | 0.4                  |
|                                  |                                                           | H <sub>2</sub>                                            | 200                         |                                            |                       |                      |
| 2nd layer                        | AlCl <sub>3</sub> /He (against SiH <sub>4</sub> )         | 1 → 0**                                                   |                             |                                            |                       |                      |
|                                  | SiH <sub>4</sub>                                          | 200                                                       |                             |                                            |                       |                      |
|                                  | C <sub>2</sub> H <sub>2</sub>                             | 10 → 20*                                                  | 250                         | 15                                         | 0.4                   | 20                   |
|                                  | NO                                                        | 1                                                         |                             |                                            |                       |                      |
| 3rd layer                        | SiH <sub>4</sub>                                          | 300                                                       |                             |                                            |                       |                      |
|                                  | H <sub>2</sub>                                            | 300                                                       | 250                         | 15                                         | 0.5                   | 10                   |

TABLE 120

| Order of lamination (layer name) | Gases and their flow rates (SCCM)                         |            | Substrate temperature (°C.) | RF discharging power (mW/cm <sup>3</sup> ) | Inner pressure (Torr) | Layer thickness (μm) |
|----------------------------------|-----------------------------------------------------------|------------|-----------------------------|--------------------------------------------|-----------------------|----------------------|
| Lower layer                      | NO                                                        | 1          |                             |                                            |                       |                      |
|                                  | SiH <sub>4</sub>                                          | 50         |                             |                                            |                       |                      |
|                                  | H <sub>2</sub>                                            | 5 → 200*   |                             |                                            |                       |                      |
|                                  | AlCl <sub>3</sub> /He<br>(S-side: 0.01 μm)                | 200 → 30** | 250                         | 1                                          | 0.4                   | 0.02                 |
|                                  | (UL-side: 0.01 μm)                                        | 30 → 10**  |                             |                                            |                       |                      |
|                                  | B <sub>2</sub> H <sub>6</sub> (against SiH <sub>4</sub> ) | 100 ppm    |                             |                                            |                       |                      |
| 1st                              | SiF <sub>4</sub>                                          | 5          |                             |                                            |                       |                      |
|                                  | SiH <sub>4</sub>                                          | 100        |                             |                                            |                       |                      |

TABLE 120-continued

| Order of lamination (layer name) | Gases and their flow rates (SCCM)                                 |                                                                                        | Substrate temperature (°C.) | RF discharging power (mW/cm <sup>3</sup> ) | Inner pressure (Torr) | Layer thickness (μm) |
|----------------------------------|-------------------------------------------------------------------|----------------------------------------------------------------------------------------|-----------------------------|--------------------------------------------|-----------------------|----------------------|
| Upper layer                      | layer 1<br>region<br>(LL-side: 2 μm)<br>(U · 2nd · LR-side: 1 μm) | B <sub>2</sub> H <sub>6</sub> (against SiH <sub>4</sub> )<br>500 ppm<br>500 ppm → 0 ** | 250                         | 10                                         | 0.4                   | 10                   |
|                                  | layer 2<br>region<br>H <sub>2</sub>                               | 200                                                                                    |                             |                                            |                       |                      |
|                                  | layer 3<br>region<br>SiH <sub>4</sub>                             | 100                                                                                    | 300                         | 15                                         | 0.4                   | 20                   |
|                                  | layer 4<br>region<br>CH <sub>4</sub>                              | 100                                                                                    |                             |                                            |                       |                      |
|                                  | layer 5<br>region<br>H <sub>2</sub>                               | 300                                                                                    | 300                         | 20                                         | 0.5                   | 5                    |
|                                  | layer 6<br>region<br>SiH <sub>4</sub>                             | 50                                                                                     | 300                         | 10                                         | 0.4                   | 0.5                  |
|                                  | layer 7<br>region<br>CH <sub>4</sub>                              | 600                                                                                    |                             |                                            |                       |                      |

TABLE 121

| Order of lamination (layer name) | Gases and their flow rates (SCCM)                                                                |                         | Substrate temperature (°C.) | RF discharging power (mW/cm <sup>3</sup> ) | Inner pressure (Torr) | Layer thickness (μm) |
|----------------------------------|--------------------------------------------------------------------------------------------------|-------------------------|-----------------------------|--------------------------------------------|-----------------------|----------------------|
| Lower layer                      | SiH <sub>4</sub><br>H <sub>2</sub>                                                               | 10 → 100*<br>5 → 200*   |                             |                                            |                       |                      |
|                                  | AlCl <sub>3</sub> /He<br>(S-side: 0.05 μm)<br>(UL-side: 0.15 μm)                                 | 200 → 40**<br>40 → 10** | 300                         | 5                                          | 0.4                   | 0.2                  |
|                                  | NH <sub>3</sub>                                                                                  | 5 → 50*                 |                             |                                            |                       |                      |
|                                  | SiF <sub>4</sub>                                                                                 | 1 → 10                  |                             |                                            |                       |                      |
| Upper layer                      | layer 1<br>region<br>SiH <sub>4</sub>                                                            | 100                     | 300                         | 5                                          | 0.4                   | 3                    |
|                                  | layer 2<br>region<br>B <sub>2</sub> H <sub>6</sub> (against SiH <sub>4</sub> )<br>H <sub>2</sub> | 200 ppm<br>500          |                             |                                            |                       |                      |
|                                  | layer 3<br>region<br>NH <sub>3</sub>                                                             | 300                     | 300                         | 15                                         | 0.4                   | 25                   |
|                                  | layer 4<br>region<br>SiH <sub>4</sub>                                                            | 50                      | 300                         | 5                                          | 0.2                   | 8                    |
|                                  | layer 5<br>region<br>H <sub>2</sub>                                                              | 100                     | 300                         | 10                                         | 0.4                   | 0.3                  |
|                                  | layer 6<br>region<br>NH <sub>3</sub>                                                             | 50                      |                             |                                            |                       |                      |

TABLE 122

| Order of lamination (layer name) | Gases and their flow rates (SCCM)                                                  |                         | Substrate temperature (°C.) | RF discharging power (mW/cm <sup>3</sup> ) | Inner pressure (Torr) | Layer thickness (μm) |
|----------------------------------|------------------------------------------------------------------------------------|-------------------------|-----------------------------|--------------------------------------------|-----------------------|----------------------|
| Lower layer                      | SiH <sub>4</sub><br>H <sub>2</sub>                                                 | 10 → 100*<br>5 → 200*   |                             |                                            |                       |                      |
|                                  | AlCl <sub>3</sub> /He<br>(S-side: 0.05 μm)<br>(UL-side: 0.15 μm)                   | 200 → 40**<br>40 → 10** | 250                         | 5                                          | 0.4                   | 0.2                  |
|                                  | NO (against SiH <sub>4</sub> )                                                     | 5 → 20*                 |                             |                                            |                       |                      |
|                                  | PH <sub>3</sub> (against SiH <sub>4</sub> )                                        | 50 ppm                  |                             |                                            |                       |                      |
|                                  | SiF <sub>4</sub>                                                                   | 1 → 10*                 |                             |                                            |                       |                      |
| Upper layer                      | layer 1<br>region<br>SiH <sub>4</sub>                                              | 100                     | 250                         | 8                                          | 0.4                   | 3                    |
|                                  | layer 2<br>region<br>PH <sub>3</sub> (against SiH <sub>4</sub> )<br>H <sub>2</sub> | 100 ppm<br>100          |                             |                                            |                       |                      |
|                                  | layer 3<br>region<br>CH <sub>4</sub>                                               | 100                     | 300                         | 10                                         | 0.4                   | 30                   |
|                                  | layer 4<br>region<br>PH <sub>3</sub> (against SiH <sub>4</sub> )                   | 50 ppm                  |                             |                                            |                       |                      |
|                                  | layer 5<br>region<br>SiH <sub>4</sub>                                              | 100                     |                             |                                            |                       |                      |
|                                  | layer 6<br>region<br>SiF <sub>4</sub>                                              | 5                       | 300                         | 3                                          | 0.5                   | 3                    |
|                                  | layer 7<br>region<br>H <sub>2</sub>                                                | 200                     |                             |                                            |                       |                      |
|                                  | layer 8<br>region<br>SiH <sub>4</sub>                                              | 50                      |                             |                                            |                       |                      |
|                                  | layer 9<br>region<br>CH <sub>4</sub>                                               | 600                     | 300                         | 10                                         | 0.4                   | 0.5                  |

TABLE 123

| Order of lamination (layer name) | Gases and their flow rates (SCCM)                                             |                                     | Substrate temperature (°C.) | RF discharging power (mW/cm <sup>3</sup> ) | Inner pressure (Torr) | Layer thickness (μm) |
|----------------------------------|-------------------------------------------------------------------------------|-------------------------------------|-----------------------------|--------------------------------------------|-----------------------|----------------------|
| Lower layer                      | N <sub>2</sub><br>SiH <sub>4</sub><br>H <sub>2</sub><br>AlCl <sub>3</sub> /He | 300<br>50<br>5 → 200*<br>200 → 20** | 250                         | 5                                          | 0.4                   | 0.05                 |

TABLE 123-continued

| Order of lamination<br>(layer name) | Gases and their flow rates<br>(SCCM)                              | Substrate temperature<br>(°C.) | RF discharging power<br>(mW/cm <sup>3</sup> ) | Inner pressure<br>(Torr) | Layer thickness<br>(μm) |
|-------------------------------------|-------------------------------------------------------------------|--------------------------------|-----------------------------------------------|--------------------------|-------------------------|
| Upper region<br>layer               | B <sub>2</sub> H <sub>6</sub> (against SiH <sub>4</sub> ) 100 ppm |                                |                                               |                          |                         |
|                                     | SiF <sub>4</sub> 5                                                |                                |                                               |                          |                         |
|                                     | SiH <sub>4</sub> 100                                              |                                |                                               |                          |                         |
|                                     | B <sub>2</sub> H <sub>6</sub> (against SiH <sub>4</sub> ) 500 ppm | 250                            | 8                                             | 0.4                      | 3                       |
|                                     | (U · 2nd · LR-side: 1 μm) 500 ppm → 0**                           |                                |                                               |                          |                         |
|                                     | H <sub>2</sub> 200                                                |                                |                                               |                          |                         |
|                                     | SiH <sub>4</sub> 300                                              |                                |                                               |                          |                         |
|                                     | C <sub>2</sub> H <sub>2</sub> 50                                  |                                |                                               |                          |                         |
|                                     | B <sub>2</sub> H <sub>6</sub> (against SiH <sub>4</sub> ) 330     |                                | 20                                            | 0.4                      | 30                      |
|                                     | (U · 1st · LR-side: 1 μm) 0 → 100 ppm**                           |                                |                                               |                          |                         |
|                                     | (U · 3rd · LR-side: 29 μm) 100 ppm                                |                                |                                               |                          |                         |
| 3rd layer                           | SiH <sub>4</sub> 200                                              |                                |                                               |                          |                         |
| layer                               | H <sub>2</sub> 200                                                | 300                            | 10                                            | 0.5                      | 10                      |
| region                              | SiH <sub>4</sub> 200                                              |                                |                                               |                          |                         |
| 4th layer                           | C <sub>2</sub> H <sub>2</sub> 200                                 | 330                            | 10                                            | 0.4                      | 1                       |
| region                              |                                                                   |                                |                                               |                          |                         |

TABLE 124

| Order of lamination<br>(layer name) | Gases and their flow rates<br>(SCCM)                              | Substrate temperature<br>(°C.) | RF discharging power<br>(mW/cm <sup>3</sup> ) | Inner pressure<br>(Torr) | Layer thickness<br>(μm) |
|-------------------------------------|-------------------------------------------------------------------|--------------------------------|-----------------------------------------------|--------------------------|-------------------------|
| Lower layer                         | PH <sub>3</sub> (against SiH <sub>4</sub> ) 50 ppm                |                                |                                               |                          |                         |
|                                     | SiH <sub>4</sub> 10 → 100*                                        |                                |                                               |                          |                         |
|                                     | H <sub>2</sub> 5 → 200*                                           |                                |                                               |                          |                         |
|                                     | AlCl <sub>3</sub> /He (S-side: 0.05 μm) 200 → 40***               | 250                            | 5                                             | 0.4                      | 0.2                     |
|                                     | (UL-side: 0.15 μm) 40 → 10**                                      |                                |                                               |                          |                         |
|                                     | NO 50 → 200*                                                      |                                |                                               |                          |                         |
|                                     | SiF <sub>4</sub> 10 → 100*                                        |                                |                                               |                          |                         |
|                                     | SiH <sub>4</sub> 40                                               |                                |                                               |                          |                         |
|                                     | PH <sub>3</sub> (against SiH <sub>4</sub> ) 250 ppm               | 250                            | 8                                             | 0.4                      | 3                       |
|                                     | (LL-side: 2 μm) 250 ppm → 0**                                     |                                |                                               |                          |                         |
| Upper layer                         | H <sub>2</sub> 200                                                |                                |                                               |                          |                         |
|                                     | SiH <sub>4</sub> 300                                              |                                |                                               |                          |                         |
|                                     | NH <sub>3</sub> 30 → 50*                                          | 330                            | 15                                            | 0.4                      | 25                      |
|                                     | PH <sub>3</sub> (against SiH <sub>4</sub> ) 50 ppm                |                                |                                               |                          |                         |
|                                     | SiH <sub>4</sub> 100                                              |                                |                                               |                          |                         |
|                                     | H <sub>2</sub> 300                                                | 300                            | 5                                             | 0.2                      | 8                       |
|                                     | SiH <sub>4</sub> 100                                              |                                |                                               |                          |                         |
|                                     | NH <sub>3</sub> 80 → 100*                                         | 300                            | 5                                             | 0.4                      | 0.7                     |
|                                     | B <sub>2</sub> H <sub>6</sub> (against SiH <sub>4</sub> ) 500 ppm |                                |                                               |                          |                         |
|                                     |                                                                   |                                |                                               |                          |                         |

TABLE 125

| Order of lamination<br>(layer name) | Gases and their flow rates<br>(SCCM)                              | Substrate temperature<br>(°C.) | RF discharging power<br>(mW/cm <sup>3</sup> ) | Inner pressure<br>(Torr) | Layer thickness<br>(μm) |
|-------------------------------------|-------------------------------------------------------------------|--------------------------------|-----------------------------------------------|--------------------------|-------------------------|
| Lower layer                         | SiH <sub>4</sub> 50                                               |                                |                                               |                          |                         |
|                                     | H <sub>2</sub> 5 → 200*                                           |                                |                                               |                          |                         |
|                                     | AlCl <sub>3</sub> /He (S-side: 0.01 μm) 200 → 30**                | 250                            | 1                                             | 0.3                      | 0.02                    |
|                                     | (UL-side: 0.01 μm) 30 → 10**                                      |                                |                                               |                          |                         |
|                                     | N <sub>2</sub> 100                                                |                                |                                               |                          |                         |
|                                     | B <sub>2</sub> H <sub>6</sub> (against SiH <sub>4</sub> ) 100 ppm |                                |                                               |                          |                         |
|                                     | SiF <sub>4</sub> 5                                                |                                |                                               |                          |                         |
|                                     | SiH <sub>4</sub> 100                                              |                                |                                               |                          |                         |
|                                     | B <sub>2</sub> H <sub>6</sub> (against SiH <sub>4</sub> ) 500 ppm | 250                            | 10                                            | 0.4                      | 3                       |
|                                     | He 600                                                            |                                |                                               |                          |                         |
| Upper layer                         | SiH <sub>4</sub> 300                                              |                                |                                               |                          |                         |
|                                     | He 600                                                            | 250                            | 25                                            | 0.6                      | 25                      |
|                                     | B <sub>2</sub> H <sub>6</sub> 0.5 ppm                             |                                |                                               |                          |                         |
|                                     | SiH <sub>4</sub> 50                                               |                                |                                               |                          |                         |
|                                     | CH <sub>4</sub> 500                                               | 250                            | 10                                            | 0.4                      | 1                       |
| region                              |                                                                   |                                |                                               |                          |                         |

TABLE 126

| Order of lamination<br>(layer name) | Gases and their flow rates<br>(SCCM)                                        | Substrate temperature<br>(°C.) | RF discharging power<br>(mW/cm <sup>3</sup> ) | Inner pressure<br>(Torr) | Layer thickness<br>(μm) |
|-------------------------------------|-----------------------------------------------------------------------------|--------------------------------|-----------------------------------------------|--------------------------|-------------------------|
| Lower layer                         | SiH <sub>4</sub> 10 → 100*                                                  |                                |                                               |                          |                         |
|                                     | H <sub>2</sub> 5 → 200*                                                     |                                |                                               |                          |                         |
|                                     | AlCl <sub>3</sub> /He<br>(S-side: 0.05 μm)<br>(UL-side: 0.15 μm) 200 → 40** | 300                            | 10                                            | 0.4                      | 0.2                     |
|                                     | NO 5 → 20*                                                                  |                                |                                               |                          |                         |
|                                     | SiF <sub>4</sub> 1 → 10*                                                    |                                |                                               |                          |                         |
|                                     | SiH <sub>4</sub> 100                                                        |                                |                                               |                          |                         |
|                                     | B <sub>2</sub> H <sub>6</sub> (against SiH <sub>4</sub> ) 200 ppm           |                                |                                               |                          |                         |
|                                     | H <sub>2</sub> 500                                                          | 300                            | 8                                             | 0.4                      | 0.5                     |
|                                     | SiF <sub>4</sub> 0.5                                                        |                                |                                               |                          |                         |
|                                     | AlCl <sub>3</sub> /He 0.1                                                   |                                |                                               |                          |                         |
| Upper layer                         | SiH <sub>4</sub> 300                                                        |                                |                                               |                          |                         |
|                                     | H <sub>2</sub> 500                                                          |                                |                                               |                          |                         |
|                                     | CH <sub>4</sub> 1                                                           |                                |                                               |                          |                         |
|                                     | NO 0.1                                                                      | 300                            | 20                                            | 0.5                      | 20                      |
|                                     | B <sub>2</sub> H <sub>6</sub> 0.3 ppm                                       |                                |                                               |                          |                         |
|                                     | SiF <sub>4</sub> 0.5                                                        |                                |                                               |                          |                         |
|                                     | AlCl <sub>3</sub> /He 0.1                                                   |                                |                                               |                          |                         |
|                                     | SiH <sub>4</sub> 100                                                        |                                |                                               |                          |                         |
|                                     | CH <sub>4</sub> 600                                                         |                                |                                               |                          |                         |
|                                     | PH <sub>3</sub> (against SiH <sub>4</sub> ) 3000 ppm                        |                                |                                               |                          |                         |
| 3rd layer region                    | NO 0.1                                                                      | 300                            | 15                                            | 0.4                      | 7                       |
|                                     | SiF <sub>4</sub> 0.5                                                        |                                |                                               |                          |                         |
|                                     | AlCl <sub>3</sub> /He 0.1                                                   |                                |                                               |                          |                         |
|                                     | B <sub>2</sub> H <sub>6</sub> (against SiH <sub>4</sub> ) 0.2 ppm           |                                |                                               |                          |                         |
|                                     | SiH <sub>4</sub> 40                                                         |                                |                                               |                          |                         |
|                                     | CH <sub>4</sub> 600                                                         |                                |                                               |                          |                         |
|                                     | NO 0.1                                                                      |                                |                                               |                          |                         |
|                                     | PH <sub>3</sub> (against SiH <sub>4</sub> ) 1 ppm                           | 300                            | 10                                            | 0.4                      | 0.1                     |
|                                     | B <sub>2</sub> H <sub>6</sub> (against SiH <sub>4</sub> ) 0.1 ppm           |                                |                                               |                          |                         |
|                                     | SiF <sub>4</sub> 0.2                                                        |                                |                                               |                          |                         |
| 4th layer region                    | AlCl <sub>3</sub> /He 0.1                                                   |                                |                                               |                          |                         |

TABLE 127

| Order of lamination<br>(layer name) | Gases and their flow rates<br>(SCCM)                                                 | Substrate temperature<br>(°C.) | RF discharging power<br>(mW/cm <sup>3</sup> ) | Inner pressure<br>(Torr) | Layer thickness<br>(μm) |
|-------------------------------------|--------------------------------------------------------------------------------------|--------------------------------|-----------------------------------------------|--------------------------|-------------------------|
| Lower layer                         | SiH <sub>4</sub> 10 → 100*                                                           |                                |                                               |                          |                         |
|                                     | H <sub>2</sub> 5 → 200*                                                              |                                |                                               |                          |                         |
|                                     | AlCl <sub>3</sub> /He<br>(S-side: 0.05 μm)<br>(UL-side: 0.15 μm) 200 → 40**          | 250                            | 5                                             | 0.4                      | 0.2                     |
|                                     | NO 5 → 20*                                                                           |                                |                                               |                          |                         |
|                                     | B <sub>2</sub> H <sub>6</sub> (against SiH <sub>4</sub> ) 100 ppm                    |                                |                                               |                          |                         |
|                                     | SiF <sub>4</sub> 1 → 10*                                                             |                                |                                               |                          |                         |
|                                     | SiH <sub>4</sub> 100                                                                 |                                |                                               |                          |                         |
|                                     | B <sub>2</sub> H <sub>6</sub> (against SiH <sub>4</sub> )<br>(LL-side: 2 μm) 500 ppm |                                |                                               |                          |                         |
|                                     | (U · 2nd · LR-side: 1 μm) 500 ppm → 0**                                              | 250                            | 8                                             | 0.4                      | 3                       |
|                                     | H <sub>2</sub> 200                                                                   |                                |                                               |                          |                         |
| Upper layer                         | SiH <sub>4</sub> 0.5                                                                 |                                |                                               |                          |                         |
|                                     | AlCl <sub>3</sub> /He 0.1                                                            |                                |                                               |                          |                         |
|                                     | SiH <sub>4</sub> 100                                                                 |                                |                                               |                          |                         |
|                                     | SiF <sub>4</sub> 5                                                                   |                                |                                               |                          |                         |
|                                     | H <sub>2</sub> 200                                                                   |                                |                                               |                          |                         |
|                                     | CH <sub>4</sub> 1                                                                    | 300                            | 3                                             | 0.5                      | 3                       |
|                                     | NO 0.1                                                                               |                                |                                               |                          |                         |
|                                     | B <sub>2</sub> H <sub>6</sub> (against SiH <sub>4</sub> ) 0.3 ppm                    |                                |                                               |                          |                         |
|                                     | AlCl <sub>3</sub> /He 0.1                                                            |                                |                                               |                          |                         |
|                                     | SiH <sub>4</sub> 100                                                                 |                                |                                               |                          |                         |
| 3rd layer region                    | CH <sub>4</sub> 100                                                                  |                                |                                               |                          |                         |
|                                     | PH <sub>3</sub> (against SiH <sub>4</sub> ) 50 ppm                                   |                                |                                               |                          |                         |
|                                     | NO 0.1                                                                               | 300                            | 15                                            | 0.4                      | 30                      |
|                                     | B <sub>2</sub> H <sub>6</sub> (against SiH <sub>4</sub> ) 0.3 ppm                    |                                |                                               |                          |                         |
|                                     | SiF <sub>4</sub> 0.5                                                                 |                                |                                               |                          |                         |
|                                     | AlCl <sub>3</sub> /He 0.1                                                            |                                |                                               |                          |                         |
|                                     | SiH <sub>4</sub> 50                                                                  |                                |                                               |                          |                         |
|                                     | CH <sub>4</sub> 600                                                                  |                                |                                               |                          |                         |
|                                     | PH <sub>3</sub> (against SiH <sub>4</sub> ) 0.3 ppm                                  |                                |                                               |                          |                         |
|                                     | B <sub>2</sub> H <sub>6</sub> (against SiH <sub>4</sub> ) 0.3 ppm                    | 300                            | 10                                            | 0.4                      | 0.5                     |
| 4th layer region                    | NO 0.1                                                                               |                                |                                               |                          |                         |
|                                     | SiF <sub>4</sub> 0.5                                                                 |                                |                                               |                          |                         |
|                                     | AlCl <sub>3</sub> /He 0.1                                                            |                                |                                               |                          |                         |
|                                     | SiH <sub>4</sub> 50                                                                  |                                |                                               |                          |                         |
|                                     | CH <sub>4</sub> 600                                                                  |                                |                                               |                          |                         |

TABLE 128

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | H <sub>2</sub> S (against SiH <sub>4</sub> ) 2 ppm                |                             |                                            |                       |                      |
|                                  | SiH <sub>4</sub> 10 → 100*                                        |                             |                                            |                       |                      |
|                                  | H <sub>2</sub> 5 → 200*                                           |                             |                                            |                       |                      |
|                                  | AlCl <sub>3</sub> /He (S-side: 0.05 μm) 200 → 40**                | 300                         | 10                                         | 0.4                   | 0.2                  |
|                                  | (UL-side: 0.15 μm) 40 → 10**                                      |                             |                                            |                       |                      |
|                                  | NO 5 → 20*                                                        |                             |                                            |                       |                      |
|                                  | SiF <sub>4</sub> 10 → 100*                                        |                             |                                            |                       |                      |
|                                  | SiH <sub>4</sub> 100                                              |                             |                                            |                       |                      |
|                                  | B <sub>2</sub> H <sub>6</sub> (against SiH <sub>4</sub> ) 200 ppm |                             |                                            |                       |                      |
|                                  | H <sub>2</sub> 500                                                | 300                         | 8                                          | 0.4                   | 0.5                  |
| Upper layer                      | SiF <sub>4</sub> 0.5                                              |                             |                                            |                       |                      |
|                                  | AlCl <sub>3</sub> /He 0.1                                         |                             |                                            |                       |                      |
|                                  | H <sub>2</sub> S (against SiH <sub>4</sub> ) 1 ppm                |                             |                                            |                       |                      |
|                                  | SiH <sub>4</sub> 300                                              |                             |                                            |                       |                      |
|                                  | H <sub>2</sub> 500                                                |                             |                                            |                       |                      |
|                                  | CH <sub>4</sub> 1                                                 |                             |                                            |                       |                      |
|                                  | NO 0.1                                                            | 300                         | 20                                         | 0.5                   | 20                   |
|                                  | B <sub>2</sub> H <sub>6</sub> (against SiH <sub>4</sub> ) 0.3 ppm |                             |                                            |                       |                      |
|                                  | SiF <sub>4</sub> 0.5                                              |                             |                                            |                       |                      |
|                                  | AlCl <sub>3</sub> /He 0.1                                         |                             |                                            |                       |                      |
| 3rd layer region                 | H <sub>2</sub> S 0.5 ppm                                          |                             |                                            |                       |                      |
|                                  | SiH <sub>4</sub> 100                                              |                             |                                            |                       |                      |
|                                  | CH <sub>4</sub> 600                                               |                             |                                            |                       |                      |
|                                  | PH <sub>3</sub> (against SiH <sub>4</sub> ) 3000 ppm              |                             |                                            |                       |                      |
|                                  | NO 0.1                                                            | 300                         | 15                                         | 0.4                   | 7                    |
|                                  | SiF <sub>4</sub> 0.5                                              |                             |                                            |                       |                      |
|                                  | AlCl <sub>3</sub> /He 0.1                                         |                             |                                            |                       |                      |
|                                  | B <sub>2</sub> H <sub>6</sub> (against SiH <sub>4</sub> ) 0.2 ppm |                             |                                            |                       |                      |
|                                  | H <sub>2</sub> S (against SiH <sub>4</sub> ) 1 ppm                |                             |                                            |                       |                      |
|                                  | SiH <sub>4</sub> 40                                               |                             |                                            |                       |                      |
| 4th layer region                 | CH <sub>4</sub> 600                                               |                             |                                            |                       |                      |
|                                  | NO 0.1                                                            |                             |                                            |                       |                      |
|                                  | PH <sub>3</sub> (against SiH <sub>4</sub> ) 1 ppm                 | 300                         | 10                                         | 0.4                   | 0.1                  |
|                                  | B <sub>2</sub> H <sub>6</sub> (against SiH <sub>4</sub> ) 0.1 ppm |                             |                                            |                       |                      |
|                                  | SiF <sub>4</sub> 0.2                                              |                             |                                            |                       |                      |
|                                  | AlCl <sub>3</sub> /He 0.1                                         |                             |                                            |                       |                      |
|                                  | H <sub>2</sub> S 10 ppm                                           |                             |                                            |                       |                      |

TABLE 129

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 50                                               |                             |                                            |                       |                      |
|                                  | GeH <sub>4</sub> 5                                                |                             |                                            |                       |                      |
|                                  | H <sub>2</sub> 10 → 200*                                          | 250                         | 5                                          | 0.4                   | 0.05                 |
|                                  | AlCl <sub>3</sub> /He 120 → 40**                                  |                             |                                            |                       |                      |
|                                  | SiH <sub>4</sub> 100                                              |                             |                                            |                       |                      |
|                                  | B <sub>2</sub> H <sub>6</sub> (against SiH <sub>4</sub> ) 200 ppm | 250                         | 8                                          | 0.4                   | 3                    |
|                                  | H <sub>2</sub> 500                                                |                             |                                            |                       |                      |
|                                  | SiH <sub>4</sub> 300                                              | 250                         | 15                                         | 0.5                   | 20                   |
|                                  | H <sub>2</sub> 300                                                |                             |                                            |                       |                      |
|                                  | SiH <sub>4</sub> 50                                               |                             |                                            |                       |                      |
| Upper layer                      | CH <sub>4</sub> 500                                               | 250                         | 10                                         | 0.4                   | 0.5                  |
|                                  | SiH <sub>4</sub> 100                                              |                             |                                            |                       |                      |
|                                  | B <sub>2</sub> H <sub>6</sub> (against SiH <sub>4</sub> ) 200 ppm |                             |                                            |                       |                      |
|                                  | H <sub>2</sub> 500                                                |                             |                                            |                       |                      |
|                                  | SiH <sub>4</sub> 300                                              |                             |                                            |                       |                      |
|                                  | H <sub>2</sub> 300                                                |                             |                                            |                       |                      |
|                                  | SiH <sub>4</sub> 50                                               |                             |                                            |                       |                      |
|                                  | CH <sub>4</sub> 500                                               |                             |                                            |                       |                      |
|                                  | SiH <sub>4</sub> 100                                              |                             |                                            |                       |                      |

TABLE 130

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 50                                               |                             |                                            |                       |                      |
|                                  | AlCl <sub>3</sub> /He 120 → 40**                                  | 250                         | 5                                          | 0.4                   | 0.05                 |
|                                  | SiH <sub>4</sub> 100                                              |                             |                                            |                       |                      |
|                                  | B <sub>2</sub> H <sub>6</sub> (against SiH <sub>4</sub> ) 200 ppm | 250                         | 8                                          | 0.4                   | 3                    |
|                                  | H <sub>2</sub> 500                                                |                             |                                            |                       |                      |
|                                  | SiH <sub>4</sub> 300                                              | 250                         | 15                                         | 0.5                   | 20                   |
|                                  | H <sub>2</sub> 300                                                |                             |                                            |                       |                      |
|                                  | SiH <sub>4</sub> 50                                               |                             |                                            |                       |                      |
|                                  | CH <sub>4</sub> 500                                               | 250                         | 10                                         | 0.4                   | 0.5                  |
|                                  | SiH <sub>4</sub> 100                                              |                             |                                            |                       |                      |
| Upper layer                      | SiH <sub>4</sub> 100                                              |                             |                                            |                       |                      |
|                                  | B <sub>2</sub> H <sub>6</sub> (against SiH <sub>4</sub> ) 200 ppm |                             |                                            |                       |                      |
|                                  | H <sub>2</sub> 500                                                |                             |                                            |                       |                      |
|                                  | SiH <sub>4</sub> 300                                              |                             |                                            |                       |                      |
|                                  | H <sub>2</sub> 300                                                |                             |                                            |                       |                      |
|                                  | SiH <sub>4</sub> 50                                               |                             |                                            |                       |                      |
|                                  | CH <sub>4</sub> 500                                               |                             |                                            |                       |                      |
|                                  | SiH <sub>4</sub> 100                                              |                             |                                            |                       |                      |

TABLE 131

| Order of lamination (layer name) | Gases and their flow rates (SCCM)                                                  | Substrate temperature (°C.) | RF discharging power (mW/cm <sup>3</sup> ) | Inner pressure (Torr) | Layer thickness (μm) |
|----------------------------------|------------------------------------------------------------------------------------|-----------------------------|--------------------------------------------|-----------------------|----------------------|
| Lower layer                      | SiH <sub>4</sub> 50                                                                |                             |                                            |                       |                      |
|                                  | GeH <sub>4</sub> 5                                                                 |                             |                                            |                       |                      |
|                                  | NO 5                                                                               |                             |                                            |                       |                      |
|                                  | H <sub>2</sub> 10 → 200*                                                           | 250                         | 5                                          | 0.4                   | 0.03                 |
|                                  | AlCl <sub>3</sub> /He (S-side: 0.01 μm) 100 → 10**                                 |                             |                                            |                       |                      |
|                                  | (UL-side: 0.01 μm) 10                                                              |                             |                                            |                       |                      |
|                                  | B <sub>2</sub> H <sub>6</sub> (against SiH <sub>4</sub> ) 50 ppm                   |                             |                                            |                       |                      |
|                                  | 1st SiH <sub>4</sub> 100                                                           |                             |                                            |                       |                      |
|                                  | Upper layer region H <sub>2</sub> 500                                              | 250                         | 8                                          | 0.4                   | 3                    |
|                                  | 2nd layer region B <sub>2</sub> H <sub>6</sub> (against SiH <sub>4</sub> ) 200 ppm |                             |                                            |                       |                      |
| 2nd layer region                 | SiH <sub>4</sub> 300                                                               |                             |                                            |                       |                      |
|                                  | H <sub>2</sub> 300                                                                 | 250                         | 15                                         | 0.5                   | 20                   |
|                                  | 3rd layer region SiH <sub>4</sub> 50                                               | 250                         | 10                                         | 0.4                   | 0.5                  |
|                                  | CH <sub>4</sub> 500                                                                |                             |                                            |                       |                      |

TABLE 132

| Order of lamination (layer name) | Gases and their flow rates (SCCM)                                                    | Substrate temperature (°C.) | RF discharging power (mW/cm <sup>3</sup> ) | Inner pressure (Torr) | Layer thickness (μm) |
|----------------------------------|--------------------------------------------------------------------------------------|-----------------------------|--------------------------------------------|-----------------------|----------------------|
| Lower layer                      | SiH <sub>4</sub> 50                                                                  |                             |                                            |                       |                      |
|                                  | B <sub>2</sub> H <sub>6</sub> (against SiH <sub>4</sub> ) 100 ppm                    |                             |                                            |                       |                      |
|                                  | SiF <sub>4</sub> 5                                                                   |                             |                                            |                       |                      |
|                                  | GeH <sub>4</sub> 10                                                                  | 150                         | 0.5                                        |                       |                      |
|                                  | H <sub>2</sub> 5 → 200*                                                              | ↓                           | ↓                                          | 0.3                   | 0.02                 |
|                                  | AlCl <sub>3</sub> /He (S-side: 0.01 μm) 200 → 30**                                   | 300                         | 1.5                                        |                       |                      |
|                                  | (UL-side: 0.01 μm) 30 → 10**                                                         |                             |                                            |                       |                      |
|                                  | 1st layer region SiH <sub>4</sub> 100                                                |                             |                                            |                       |                      |
|                                  | H <sub>2</sub> 200                                                                   |                             |                                            |                       |                      |
|                                  | Upper layer region B <sub>2</sub> H <sub>6</sub> (against SiH <sub>4</sub> ) 500 ppm | 250                         | 10                                         | 0.4                   | 3                    |
| 2nd layer region                 | (LL-side: 2 μm) 500 ppm                                                              |                             |                                            |                       |                      |
|                                  | (U · 2nd · LR-side: 1 μm) 500 ppm → 10**                                             |                             |                                            |                       |                      |
| 2nd layer region                 | SiH <sub>4</sub> 300                                                                 |                             |                                            |                       |                      |
|                                  | H <sub>2</sub> 500                                                                   | 250                         | 20                                         | 0.5                   | 20                   |

TABLE 133

| Order of lamination (layer name) | Gases and their flow rates (SCCM)                                                    | Substrate temperature (°C.) | RF discharging power (mW/cm <sup>3</sup> ) | Inner pressure (Torr) | Layer thickness (μm) |
|----------------------------------|--------------------------------------------------------------------------------------|-----------------------------|--------------------------------------------|-----------------------|----------------------|
| Lower layer                      | SiH <sub>4</sub> 50                                                                  |                             |                                            |                       |                      |
|                                  | GeH <sub>4</sub> 5                                                                   |                             |                                            |                       |                      |
|                                  | B <sub>2</sub> H <sub>6</sub> (against SiH <sub>4</sub> ) 100 ppm                    |                             |                                            |                       |                      |
|                                  | H <sub>2</sub> 5 → 200*                                                              | 250                         | 1                                          | 0.3                   | 0.02                 |
|                                  | AlCl <sub>3</sub> /He (S-side: 0.01 μm) 200 → 30**                                   |                             |                                            |                       |                      |
|                                  | (UL-side: 0.01 μm) 30 → 10**                                                         |                             |                                            |                       |                      |
|                                  | 1st layer region SiH <sub>4</sub> 100                                                |                             |                                            |                       |                      |
|                                  | He 600                                                                               |                             |                                            |                       |                      |
|                                  | Upper layer region B <sub>2</sub> H <sub>6</sub> (against SiH <sub>4</sub> ) 500 ppm | 250                         | 10                                         | 0.4                   | 3                    |
|                                  | AlCl <sub>3</sub> /He 0.1                                                            |                             |                                            |                       |                      |
| 2nd layer region                 | SiF <sub>4</sub> 0.5                                                                 |                             |                                            |                       |                      |
|                                  | SiH <sub>4</sub> 300                                                                 |                             |                                            |                       |                      |
|                                  | He 600                                                                               |                             |                                            |                       |                      |
|                                  | B <sub>2</sub> H <sub>6</sub> (against SiH <sub>4</sub> ) 0.3 ppm                    |                             |                                            |                       |                      |
|                                  | AlCl <sub>3</sub> /He 0.1                                                            | 250                         | 25                                         | 0.6                   | 25                   |
|                                  | SiF <sub>4</sub> 0.5                                                                 |                             |                                            |                       |                      |
| 3rd layer region                 | CH <sub>4</sub> 1                                                                    |                             |                                            |                       |                      |
|                                  | NO 0.1                                                                               |                             |                                            |                       |                      |
|                                  | GeH <sub>4</sub> 0.1                                                                 |                             |                                            |                       |                      |
|                                  | SiH <sub>4</sub> 50                                                                  |                             |                                            |                       |                      |
|                                  | CH <sub>4</sub> 500                                                                  |                             |                                            |                       |                      |
|                                  | NO 0.1                                                                               |                             |                                            |                       |                      |
|                                  | GeH <sub>4</sub> 0.1                                                                 | 250                         | 10                                         | 0.4                   | 1                    |
|                                  | B <sub>2</sub> H <sub>6</sub> (against SiH <sub>4</sub> ) 0.3 ppm                    |                             |                                            |                       |                      |
|                                  | Al <sub>2</sub> Cl <sub>3</sub> /He 0.1                                              |                             |                                            |                       |                      |
|                                  | SiF <sub>4</sub> 0.5                                                                 |                             |                                            |                       |                      |

TABLE 134

| Order of lamination (layer name) | Gases and their flow rates (SCCM)                                  | Substrate temperature (°C.) | RF discharging power (mW/cm <sup>3</sup> ) | Inner pressure (Torr) | Layer thickness (μm) |
|----------------------------------|--------------------------------------------------------------------|-----------------------------|--------------------------------------------|-----------------------|----------------------|
| Lower layer                      | CH <sub>4</sub> 50 → 200*                                          |                             |                                            |                       |                      |
|                                  | GeH <sub>4</sub> 1 → 10*                                           |                             |                                            |                       |                      |
|                                  | SiH <sub>4</sub> 10 → 100*                                         |                             |                                            |                       |                      |
|                                  | H <sub>2</sub> 5 → 200*                                            | 250                         | 10                                         | 0.4                   | 0.2                  |
|                                  | Al(CH <sub>3</sub> ) <sub>3</sub> /He (S-side: 0.05 μm) 200 → 40** |                             |                                            |                       |                      |
|                                  | (UL-side: 0.15 μm) 40 → 10**                                       |                             |                                            |                       |                      |
| 1st layer                        | SiH <sub>4</sub> 100                                               |                             |                                            |                       |                      |
|                                  | H <sub>2</sub> 200                                                 |                             |                                            |                       |                      |
|                                  | B <sub>2</sub> H <sub>6</sub> (against SiH <sub>4</sub> ) 500 ppm  | 250                         | 10                                         | 0.4                   | 3                    |
| Upper region                     | (LL-side: 2 μm) 500 ppm                                            |                             |                                            |                       |                      |
|                                  | (U + 2nd + LR-side: 1 μm) 500 ppm → 0**                            |                             |                                            |                       |                      |
|                                  | SiH <sub>4</sub> 400                                               |                             |                                            |                       |                      |
| 2nd layer region                 | Ar 200                                                             | 250                         | 10                                         | 0.5                   | 15                   |
|                                  | SiH <sub>4</sub> 100                                               |                             |                                            |                       |                      |
| 3rd layer region                 | NH <sub>3</sub> 30                                                 | 250                         | 5                                          | 0.4                   | 0.3                  |

TABLE 135

| Order of Lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | NO 5 → 20*                                                        |                             |                                            |                       |                      |
|                                  | GeF <sub>4</sub> 1 → 10*                                          |                             |                                            |                       |                      |
|                                  | SiH <sub>4</sub> 10 → 100*                                        |                             |                                            |                       |                      |
|                                  | H <sub>2</sub> 5 → 200*                                           | 300                         | 10                                         | 0.4                   | 0.2                  |
|                                  | AlCl <sub>3</sub> /He (S-side: 0.05 μm) 200 → 40**                |                             |                                            |                       |                      |
|                                  | (UL-side: 0.15 μm) 40 → 10**                                      |                             |                                            |                       |                      |
| 1st layer region                 | SiH <sub>4</sub> 100                                              |                             |                                            |                       |                      |
|                                  | H <sub>2</sub> 500                                                | 300                         | 8                                          | 0.4                   | 0.5                  |
|                                  | B <sub>2</sub> H <sub>6</sub> (against SiH <sub>4</sub> ) 200 ppm |                             |                                            |                       |                      |
| Upper layer                      | SiH <sub>4</sub> 300                                              |                             |                                            |                       |                      |
|                                  | H <sub>2</sub> 500                                                | 300                         | 20                                         | 0.5                   | 20                   |
|                                  | SiH <sub>4</sub> 100                                              |                             |                                            |                       |                      |
| 3rd layer region                 | CH <sub>4</sub> 600                                               | 300                         | 15                                         | 0.4                   | 7                    |
|                                  | PH <sub>3</sub> (against SiH <sub>4</sub> ) 3000 ppm              |                             |                                            |                       |                      |
| 4th layer region                 | SiH <sub>4</sub> 40                                               |                             |                                            |                       |                      |
|                                  | CH <sub>4</sub> 600                                               | 300                         | 10                                         | 0.4                   | 0.1                  |

TABLE 136

| Order of lamination (layer name) | Gases and their flow rates (SCCM)                                  | Substrate temperature (°C.) | RF discharging power (mW/cm <sup>3</sup> ) | Inner pressure (Torr) | Layer thickness (μm) |
|----------------------------------|--------------------------------------------------------------------|-----------------------------|--------------------------------------------|-----------------------|----------------------|
| Lower layer                      | SiH <sub>4</sub> 50                                                |                             |                                            |                       |                      |
|                                  | GeH <sub>4</sub> 5                                                 |                             |                                            |                       |                      |
|                                  | PF <sub>5</sub> (against SiH <sub>4</sub> ) 50 ppm                 |                             |                                            |                       |                      |
|                                  | NO 5                                                               | 330                         | 5                                          | 0.4                   | 0.05                 |
|                                  | H <sub>2</sub> 5 → 200*                                            |                             |                                            |                       |                      |
|                                  | AlCl <sub>3</sub> /He 200 → 20**                                   |                             |                                            |                       |                      |
| Upper layer                      | SiH <sub>4</sub> 100                                               |                             |                                            |                       |                      |
|                                  | H <sub>2</sub> 100                                                 | 330                         | 8                                          | 0.4                   | 3                    |
|                                  | PF <sub>5</sub> (against SiH <sub>4</sub> ) 100 ppm                |                             |                                            |                       |                      |
|                                  | SiH <sub>4</sub> 400                                               |                             |                                            |                       |                      |
|                                  | SiF <sub>4</sub> 10                                                | 330                         | 25                                         | 0.5                   | 25                   |
|                                  | H <sub>2</sub> 800                                                 |                             |                                            |                       |                      |
| Upper layer                      | SiH <sub>4</sub> 100                                               |                             |                                            |                       |                      |
|                                  | CH <sub>4</sub> 400                                                | 350                         | 15                                         | 0.4                   | 5                    |
|                                  | B <sub>2</sub> H <sub>6</sub> (against SiH <sub>4</sub> ) 5000 ppm |                             |                                            |                       |                      |
|                                  | SiH <sub>4</sub> 20                                                |                             |                                            |                       |                      |
|                                  | CH <sub>4</sub> 400                                                | 350                         | 10                                         | 0.4                   | 1                    |
|                                  | B <sub>2</sub> H <sub>6</sub> (against SiH <sub>4</sub> ) 8000 ppm |                             |                                            |                       |                      |

TABLE 137

| Order of lamination<br>(layer name) | Gases and<br>their flow rates<br>(SCCM)                           | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|-------------------------------------------------------------------|-----------------------------------|--------------------------------------------------|-----------------------------|----------------------------|
| Lower layer                         | SiH <sub>4</sub> 50                                               |                                   |                                                  |                             |                            |
|                                     | GeH <sub>4</sub> 5                                                |                                   |                                                  |                             |                            |
|                                     | H <sub>2</sub> S (against SiH <sub>4</sub> ) 10 ppm               |                                   |                                                  |                             |                            |
|                                     | H <sub>2</sub> 5 → 200*                                           | 300                               | 1                                                | 0.3                         | 0.02                       |
|                                     | AlCl <sub>3</sub> /He<br>(S-side: 0.01 μm)                        |                                   |                                                  |                             |                            |
|                                     | (UL-side: 0.01 μm) 200 → 30**                                     |                                   |                                                  |                             |                            |
| Upper layer                         | SiH <sub>4</sub> 30 → 10**                                        |                                   |                                                  |                             |                            |
|                                     | 1st SiH <sub>4</sub> 100                                          |                                   |                                                  |                             |                            |
|                                     | H <sub>2</sub> 200                                                | 300                               | 8                                                | 0.4                         | 5                          |
|                                     | B <sub>2</sub> H <sub>6</sub> (against SiH <sub>4</sub> ) 200 ppm |                                   |                                                  |                             |                            |
|                                     | 2nd SiH <sub>4</sub> 300                                          |                                   |                                                  |                             |                            |
|                                     | H <sub>2</sub> 200                                                | 300                               | 20                                               | 0.5                         | 20                         |
| layer region                        | 3rd SiH <sub>4</sub> 50                                           |                                   |                                                  |                             |                            |
|                                     | N <sub>2</sub> 500                                                | 300                               | 20                                               | 0.4                         | 5                          |
|                                     | PH <sub>3</sub> (against SiH <sub>4</sub> ) 3000 ppm              |                                   |                                                  |                             |                            |
|                                     | 4th SiH <sub>4</sub> 40                                           |                                   |                                                  |                             |                            |
|                                     | CH <sub>4</sub> 600                                               | 300                               | 10                                               | 0.4                         | 0.3                        |
|                                     |                                                                   |                                   |                                                  |                             |                            |

TABLE 138

| Order of lamination<br>(layer name) | Gases and<br>their flow rates<br>(SCCM)                           | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|-------------------------------------------------------------------|-----------------------------------|--------------------------------------------------|-----------------------------|----------------------------|
| Lower layer                         | SiH <sub>4</sub> 50                                               |                                   |                                                  |                             |                            |
|                                     | B <sub>2</sub> H <sub>6</sub> (against SiH <sub>4</sub> ) 100 ppm |                                   |                                                  |                             |                            |
|                                     | C <sub>2</sub> H <sub>2</sub> 10                                  |                                   |                                                  |                             |                            |
|                                     | NO 5                                                              | 250                               | 5                                                | 0.4                         | 0.05                       |
|                                     | GeF <sub>4</sub> 5                                                |                                   |                                                  |                             |                            |
|                                     | H <sub>2</sub> 5 → 200*                                           |                                   |                                                  |                             |                            |
| Upper layer                         | AlCl <sub>3</sub> /He 200 → 20**                                  |                                   |                                                  |                             |                            |
|                                     | 1st SiH <sub>4</sub> 100                                          |                                   |                                                  |                             |                            |
|                                     | H <sub>2</sub> 200                                                |                                   |                                                  |                             |                            |
|                                     | B <sub>2</sub> H <sub>6</sub> (against SiH <sub>4</sub> ) 500 ppm | 250                               | 10                                               | 0.4                         | 5                          |
|                                     | (LL-side: 3 μm)<br>(U · 2nd · LR-side: 2 μm)                      |                                   |                                                  |                             |                            |
|                                     | AlCl <sub>3</sub> /He 500 ppm → 0**<br>1 → 10*                    |                                   |                                                  |                             |                            |
| layer region                        | 2nd SiH <sub>4</sub> 300                                          |                                   |                                                  |                             |                            |
|                                     | H <sub>2</sub> 300                                                | 250                               | 15                                               | 0.5                         | 10                         |
|                                     | 3rd SiH <sub>4</sub> 200                                          |                                   |                                                  |                             |                            |
|                                     | C <sub>2</sub> H <sub>2</sub> 10 → 20*                            | 250                               | 15                                               | 0.4                         | 20                         |
|                                     | NO 1                                                              |                                   |                                                  |                             |                            |
|                                     |                                                                   |                                   |                                                  |                             |                            |

TABLE 139

| Order of lamination<br>(layer name) | Gases and<br>their flow rates<br>(SCCM)                                  | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|--------------------------------------------------------------------------|-----------------------------------|--------------------------------------------------|-----------------------------|----------------------------|
| Lower layer                         | SiH <sub>4</sub> 50                                                      |                                   |                                                  |                             |                            |
|                                     | BF <sub>3</sub> (against SiH <sub>4</sub> ) 100 ppm                      |                                   |                                                  |                             |                            |
|                                     | NO 1                                                                     |                                   |                                                  |                             |                            |
|                                     | GeH <sub>4</sub> 5                                                       |                                   |                                                  |                             |                            |
|                                     | H <sub>2</sub> 5 → 200*                                                  | 250                               | 1                                                | 0.4                         | 0.02                       |
|                                     | AlCl <sub>3</sub> /He (S-side: 0.01 μm)<br>(UL-side: 0.01 μm) 200 → 30** |                                   |                                                  |                             |                            |
| Upper layer                         | 30 → 10**                                                                |                                   |                                                  |                             |                            |
|                                     | 1st SiH <sub>4</sub> 100                                                 |                                   |                                                  |                             |                            |
|                                     | H <sub>2</sub> 200                                                       |                                   |                                                  |                             |                            |
|                                     | B <sub>2</sub> H <sub>6</sub> (against SiH <sub>4</sub> ) 500 ppm        | 250                               | 10                                               | 0.4                         | 10                         |
|                                     | (LL-side: 8 μm)<br>(U · 2nd · LR-side: 2 μm)                             |                                   |                                                  |                             |                            |
|                                     | 2nd SiH <sub>4</sub> 300 → 0 ppm**<br>H <sub>2</sub> 300                 | 300                               | 20                                               | 0.5                         | 5                          |
| layer region                        | 3rd SiH <sub>4</sub> 100                                                 |                                   |                                                  |                             |                            |
|                                     | CH <sub>4</sub> 100                                                      | 300                               | 15                                               | 0.4                         | 20                         |
|                                     | 4th SiH <sub>4</sub> 50                                                  |                                   |                                                  |                             |                            |
|                                     |                                                                          |                                   |                                                  |                             |                            |

TABLE 139-continued

| Order of lamination<br>(layer name) | Gases and their flow rates<br>(SCCM) | Substrate temperature<br>(°C.) | RF discharging power<br>(mW/cm <sup>3</sup> ) | Inner pressure<br>(Torr) | Layer thickness<br>(μm) |
|-------------------------------------|--------------------------------------|--------------------------------|-----------------------------------------------|--------------------------|-------------------------|
| layer region                        | CH <sub>4</sub>                      | 600                            | 300                                           | 10                       | 0.4                     |
|                                     |                                      |                                |                                               |                          | 0.5                     |

TABLE 140

| Order of lamination<br>(layer name) | Gases and their flow rates<br>(SCCM)       | Substrate temperature<br>(°C.)                            | RF discharging power<br>(mW/cm <sup>3</sup> ) | Inner pressure<br>(Torr) | Layer thickness<br>(μm) |
|-------------------------------------|--------------------------------------------|-----------------------------------------------------------|-----------------------------------------------|--------------------------|-------------------------|
| Lower layer                         | SiH <sub>4</sub>                           | 10 → 100*                                                 |                                               |                          |                         |
|                                     | GeF <sub>4</sub>                           | 1 → 10*                                                   |                                               |                          |                         |
|                                     | NH <sub>3</sub>                            | 5 → 50*                                                   |                                               |                          |                         |
|                                     | H <sub>2</sub>                             | 5 → 200*                                                  | 300                                           | 5                        | 0.4                     |
|                                     | AlCl <sub>3</sub> /He<br>(S-side: 0.05 μm) | 200 → 40**                                                |                                               |                          | 0.2                     |
|                                     | (UL-side: 0.15 μm)                         | 40 → 10**                                                 |                                               |                          |                         |
| Upper layer                         | 1st layer                                  | SiH <sub>4</sub>                                          | 100                                           |                          |                         |
|                                     |                                            | H <sub>2</sub>                                            | 500                                           | 300                      | 5                       |
|                                     |                                            | B <sub>2</sub> H <sub>6</sub> (against SiH <sub>4</sub> ) | 200 ppm                                       |                          |                         |
|                                     | 2nd layer                                  | SiH <sub>4</sub>                                          | 100                                           |                          |                         |
|                                     |                                            | H <sub>2</sub>                                            | 300                                           | 300                      | 5                       |
|                                     | 3rd layer                                  | SiH <sub>4</sub>                                          | 300                                           |                          |                         |
|                                     |                                            | NH <sub>3</sub>                                           | 50                                            | 300                      | 15                      |
|                                     | 4th layer                                  | SiH <sub>4</sub>                                          | 100                                           |                          |                         |
|                                     |                                            | NH <sub>3</sub>                                           | 50                                            | 300                      | 10                      |
|                                     |                                            |                                                           |                                               | 0.4                      | 0.4                     |
|                                     |                                            |                                                           |                                               | 0.3                      |                         |

TABLE 141

| Order of lamination<br>(layer name) | Gases and their flow rates<br>(SCCM)                      | Substrate temperature<br>(°C.)                            | RF discharging power<br>(mW/cm <sup>3</sup> ) | Inner pressure<br>(Torr) | Layer thickness<br>(μm) |
|-------------------------------------|-----------------------------------------------------------|-----------------------------------------------------------|-----------------------------------------------|--------------------------|-------------------------|
| Lower layer                         | SiH <sub>4</sub>                                          | 10 → 100*                                                 |                                               |                          |                         |
|                                     | B <sub>2</sub> H <sub>6</sub> (against SiH <sub>4</sub> ) | 100 ppm                                                   |                                               |                          |                         |
|                                     | NO                                                        | 5 → 20*                                                   |                                               |                          |                         |
|                                     | GeH <sub>4</sub>                                          | 5 → 10*                                                   | 250                                           | 5                        | 0.4                     |
|                                     | H <sub>2</sub>                                            | 5 → 200*                                                  |                                               |                          |                         |
|                                     | AlCl <sub>3</sub> /He<br>(S-side: 0.05 μm)                | 200 → 40**                                                |                                               |                          | 0.2                     |
|                                     | (UL-side: 0.15 μm)                                        | 40 → 10**                                                 |                                               |                          |                         |
| Upper layer                         | 1st layer                                                 | SiH <sub>4</sub>                                          | 100                                           |                          |                         |
|                                     |                                                           | H <sub>2</sub>                                            | 200                                           |                          |                         |
|                                     |                                                           | B <sub>2</sub> H <sub>6</sub> (against SiH <sub>4</sub> ) | 250                                           | 8                        | 0.4                     |
|                                     | (LL-side: 2 μm)                                           | 500 ppm                                                   |                                               |                          | 3                       |
|                                     | (U + 2nd + LR-side: 1 μm)                                 | 500 → 0 ppm**                                             |                                               |                          |                         |
|                                     | 2nd layer                                                 | SiH <sub>4</sub>                                          | 100                                           |                          |                         |
|                                     |                                                           | SiF <sub>4</sub>                                          | 5                                             | 3                        | 0.5                     |
|                                     | region                                                    | H <sub>2</sub>                                            | 200                                           |                          | 3                       |
|                                     | 3rd layer                                                 | SiH <sub>4</sub>                                          | 100                                           |                          |                         |
|                                     |                                                           | CH <sub>4</sub>                                           | 100                                           | 15                       | 0.4                     |
|                                     | region                                                    | PH <sub>3</sub> (against SiH <sub>4</sub> )               | 50 ppm                                        |                          | 30                      |
|                                     | 4th layer                                                 | SiH <sub>4</sub>                                          | 50                                            |                          |                         |
|                                     |                                                           | CH <sub>4</sub>                                           | 600                                           | 10                       | 0.4                     |
|                                     | region                                                    |                                                           |                                               | 0.5                      |                         |

TABLE 142

| Order of lamination<br>(layer name) | Gases and their flow rates<br>(SCCM)        | Substrate temperature<br>(°C.) | RF discharging power<br>(mW/cm <sup>3</sup> ) | Inner pressure<br>(Torr) | Layer thickness<br>(μm) |
|-------------------------------------|---------------------------------------------|--------------------------------|-----------------------------------------------|--------------------------|-------------------------|
| Lower layer                         | SiH <sub>4</sub>                            | 50                             |                                               |                          |                         |
|                                     | PH <sub>3</sub> (against SiH <sub>4</sub> ) | 50 ppm                         |                                               |                          |                         |
|                                     | Si <sub>2</sub> F <sub>6</sub>              | 5                              | 250                                           | 5                        | 0.4                     |
|                                     | GeH <sub>4</sub>                            | 10                             |                                               |                          |                         |
|                                     | H <sub>2</sub>                              | 5 → 200*                       |                                               |                          |                         |
|                                     | AlCl <sub>3</sub> /He                       | 200 → 20**                     |                                               |                          |                         |
| 1st layer                           | SiH <sub>4</sub>                            | 40                             |                                               |                          |                         |
|                                     | H <sub>2</sub>                              | 40                             |                                               |                          |                         |

TABLE 142-continued

| Order of lamination (layer name) | Gases and their flow rates (SCCM)                                                           | Substrate temperature (°C.) | RF discharging power (mW/cm <sup>3</sup> ) | Inner pressure (Torr) | Layer thickness (μm) |
|----------------------------------|---------------------------------------------------------------------------------------------|-----------------------------|--------------------------------------------|-----------------------|----------------------|
| Upper layer                      | PH <sub>3</sub> (against SiH <sub>4</sub> )<br>(LL-side: 2 μm)<br>(U · 2nd · LR-side: 1 μm) | 250 ppm                     | 250                                        | 8                     | 0.4                  |
| 2nd layer                        | Si <sub>2</sub> H <sub>6</sub><br>H <sub>2</sub>                                            | 200<br>200                  | 300                                        | 10                    | 0.5                  |
| region                           |                                                                                             |                             |                                            |                       | 10                   |
| 3rd layer                        | SiH <sub>4</sub><br>C <sub>2</sub> H <sub>2</sub>                                           | 300<br>50                   |                                            |                       |                      |
| region                           | B <sub>2</sub> H <sub>6</sub> (against SiH <sub>4</sub> )<br>(U · 2nd · LR-side: 1 μm)      | 0 → 100 ppm*                | 330                                        | 20                    | 0.4                  |
|                                  | (U · 4th · LT-side: 29 μm)                                                                  | 100 ppm                     |                                            |                       | 30                   |
| 4th layer                        | SiH <sub>4</sub><br>C <sub>2</sub> H <sub>2</sub>                                           | 200<br>200                  | 330                                        | 10                    | 0.4                  |
| region                           |                                                                                             |                             |                                            |                       | 1                    |

TABLE 143

| Order of lamination (layer name) | Gases and their flow rates (SCCM)                                                                                                                                                                         | Substrate temperature (°C.)                                                                         | RF discharging power (mW/cm <sup>3</sup> ) | Inner pressure (Torr) | Layer thickness (μm) |
|----------------------------------|-----------------------------------------------------------------------------------------------------------------------------------------------------------------------------------------------------------|-----------------------------------------------------------------------------------------------------|--------------------------------------------|-----------------------|----------------------|
| Lower layer                      | Si <sub>2</sub> F <sub>6</sub><br>B <sub>2</sub> H <sub>6</sub> (against SiH <sub>4</sub> )<br>NO<br>GeH <sub>4</sub><br>SiH <sub>4</sub><br>H <sub>2</sub><br>AlCl <sub>3</sub> /He<br>(S-side: 0.05 μm) | 1 → 5*<br>80 ppm<br>5 → 20*<br>1 → 10*<br>10 → 100*<br>5 → 200*<br>200 → 40**<br>(UL-side: 0.15 μm) | 250                                        | 5                     | 0.4                  |
|                                  |                                                                                                                                                                                                           | 40 → 10**                                                                                           |                                            |                       | 0.2                  |
| Upper layer                      | 1st layer                                                                                                                                                                                                 | SiH <sub>4</sub><br>H <sub>2</sub>                                                                  | 100<br>500                                 | 300                   | 8                    |
|                                  | region                                                                                                                                                                                                    | B <sub>2</sub> H <sub>6</sub> (against SiH <sub>4</sub> )                                           | 200 ppm                                    |                       | 3                    |
|                                  | 2nd layer                                                                                                                                                                                                 | SiH <sub>4</sub><br>H <sub>2</sub>                                                                  | 100<br>300                                 | 300                   | 5                    |
|                                  | region                                                                                                                                                                                                    |                                                                                                     |                                            | 0.2                   | 8                    |
|                                  | 3rd layer                                                                                                                                                                                                 | SiH <sub>4</sub><br>NH <sub>3</sub>                                                                 | 300<br>30 → 50*                            | 300                   | 15                   |
|                                  | region                                                                                                                                                                                                    | PH <sub>3</sub> (against SiH <sub>4</sub> )                                                         | 50 ppm                                     |                       | 0.4                  |
|                                  | 4th layer                                                                                                                                                                                                 | SiH <sub>4</sub><br>NH <sub>3</sub>                                                                 | 100<br>80 → 100*                           | 300                   | 5                    |
|                                  | region                                                                                                                                                                                                    | PH <sub>3</sub> (against SiH <sub>4</sub> )                                                         | 500 ppm                                    |                       | 0.4                  |

TABLE 144

| Order of lamination (layer name) | Gases and their flow rates (SCCM)                                                                          | Substrate temperature (°C.)                                  | RF discharging power (mW/cm <sup>3</sup> ) | Inner pressure (Torr) | Layer thickness (μm) |
|----------------------------------|------------------------------------------------------------------------------------------------------------|--------------------------------------------------------------|--------------------------------------------|-----------------------|----------------------|
| Lower layer                      | NO<br>GeH <sub>4</sub><br>SiH <sub>4</sub><br>H <sub>2</sub><br>AlCl <sub>3</sub> /He<br>(S-side: 0.01 μm) | 5<br>5<br>50<br>5 → 200*<br>200 → 30**<br>(UL-side: 0.01 μm) | 250                                        | 1                     | 0.4                  |
|                                  |                                                                                                            | 30 → 10**                                                    |                                            |                       | 0.02                 |
| Upper layer                      | 1st layer                                                                                                  | SiH <sub>4</sub><br>H <sub>2</sub>                           | 100<br>100                                 | 300                   | 8                    |
|                                  | region                                                                                                     | PH <sub>3</sub> (against SiH <sub>4</sub> )                  | 100 ppm                                    |                       | 0.4                  |
|                                  | 2nd layer                                                                                                  | SiH <sub>4</sub><br>H <sub>2</sub>                           | 300<br>500                                 | 300                   | 20                   |
|                                  | region                                                                                                     |                                                              |                                            | 0.5                   | 20                   |
|                                  | 3rd layer                                                                                                  | SiH <sub>4</sub><br>GeH <sub>4</sub>                         | 100<br>10 → 50*                            | 300                   | 5                    |
|                                  | region                                                                                                     | H <sub>2</sub>                                               | 300                                        |                       | 0.4                  |
|                                  | 4th layer                                                                                                  | SiH <sub>4</sub><br>CH <sub>4</sub>                          | 100 → 40**<br>100 → 600*                   | 300                   | 10                   |
|                                  | region                                                                                                     |                                                              |                                            | 0.4                   | 1                    |

TABLE 145

| Order of lamination<br>(layer name) | Gases and their flow rates<br>(SCCM)                              | Substrate temperature<br>(°C.)   | RF discharging power<br>(mW/cm <sup>3</sup> ) | Inner pressure<br>(Torr) | Layer thickness<br>(μm) |
|-------------------------------------|-------------------------------------------------------------------|----------------------------------|-----------------------------------------------|--------------------------|-------------------------|
| Lower layer                         | B <sub>2</sub> H <sub>6</sub> (against SiH <sub>4</sub> ) 50 ppm  |                                  |                                               |                          |                         |
|                                     | NO 5                                                              |                                  |                                               |                          |                         |
|                                     | GeH <sub>4</sub> 5                                                |                                  |                                               |                          |                         |
|                                     | SiH <sub>4</sub> 50                                               |                                  |                                               |                          |                         |
|                                     | H <sub>2</sub> 5 → 200*                                           | 300                              | 1                                             | 0.3                      | 0.02                    |
|                                     | AlCl <sub>3</sub> /He<br>(S-side: 0.01 μm)                        | 200 → 30**<br>(UL-side: 0.01 μm) |                                               |                          |                         |
| Upper layer                         | SiH <sub>4</sub> 100                                              |                                  |                                               |                          |                         |
|                                     | H <sub>2</sub> 500                                                | 300                              | 8                                             | 0.4                      | 10                      |
|                                     | B <sub>2</sub> H <sub>6</sub> (against SiH <sub>4</sub> ) 200 ppm |                                  |                                               |                          |                         |
|                                     | SiH <sub>4</sub> 300                                              |                                  |                                               |                          |                         |
|                                     | H <sub>2</sub> 400                                                | 300                              | 15                                            | 0.5                      | 20                      |
|                                     | SiH <sub>4</sub> 50                                               |                                  |                                               |                          |                         |
| 1st layer region                    | CH <sub>4</sub> 500                                               | 300                              | 10                                            | 0.4                      | 0.5                     |
|                                     |                                                                   |                                  |                                               |                          |                         |
| 2nd layer region                    | SiH <sub>4</sub> 80                                               |                                  |                                               |                          |                         |
|                                     | H <sub>2</sub> 400                                                | 300                              | 7                                             | 0.3                      | 10                      |
|                                     | B <sub>2</sub> H <sub>6</sub> (against SiH <sub>4</sub> ) 200 ppm |                                  |                                               |                          |                         |
|                                     | SiH <sub>4</sub> 200                                              |                                  |                                               |                          |                         |
|                                     | H <sub>2</sub> 400                                                | 300                              | 12                                            | 0.4                      | 20                      |
|                                     | SiH <sub>4</sub> 40                                               |                                  |                                               |                          |                         |
| 3rd layer region                    | CH <sub>4</sub> 400                                               | 300                              | 7                                             | 0.3                      | 0.5                     |
|                                     |                                                                   |                                  |                                               |                          |                         |

TABLE 146

| Order of lamination<br>(layer name) | Gases and their flow rates<br>(SCCM)                              | Substrate temperature<br>(°C.)   | RF discharging power<br>(mW/cm <sup>3</sup> ) | Inner pressure<br>(Torr) | Layer thickness<br>(μm) |
|-------------------------------------|-------------------------------------------------------------------|----------------------------------|-----------------------------------------------|--------------------------|-------------------------|
| Lower layer                         | GeH <sub>4</sub> 5                                                |                                  |                                               |                          |                         |
|                                     | B <sub>2</sub> H <sub>6</sub> (against SiH <sub>4</sub> ) 50 ppm  |                                  |                                               |                          |                         |
|                                     | NO 5                                                              |                                  |                                               |                          |                         |
|                                     | H <sub>2</sub> 5 → 200*                                           | 300                              | 0.7                                           | 0.3                      | 0.02                    |
|                                     | AlCl <sub>3</sub> /He<br>(S-side: 0.01 μm)                        | 200 → 30**<br>(UL-side: 0.01 μm) |                                               |                          |                         |
|                                     | SiH <sub>4</sub> 30 → 10**                                        |                                  |                                               |                          |                         |
| Upper layer                         | SiH <sub>4</sub> 80                                               |                                  |                                               |                          |                         |
|                                     | H <sub>2</sub> 400                                                | 300                              | 7                                             | 0.3                      | 10                      |
|                                     | B <sub>2</sub> H <sub>6</sub> (against SiH <sub>4</sub> ) 200 ppm |                                  |                                               |                          |                         |
|                                     | SiH <sub>4</sub> 200                                              |                                  |                                               |                          |                         |
|                                     | H <sub>2</sub> 400                                                | 300                              | 12                                            | 0.4                      | 20                      |
|                                     | SiH <sub>4</sub> 40                                               |                                  |                                               |                          |                         |
| 1st layer region                    | CH <sub>4</sub> 400                                               | 300                              | 7                                             | 0.3                      | 0.5                     |
|                                     |                                                                   |                                  |                                               |                          |                         |
| 2nd layer region                    | SiH <sub>4</sub> 60                                               |                                  |                                               |                          |                         |
|                                     | H <sub>2</sub> 300                                                | 300                              | 6                                             | 0.2                      | 10                      |
|                                     | B <sub>2</sub> H <sub>6</sub> (against SiH <sub>4</sub> ) 200 ppm |                                  |                                               |                          |                         |
|                                     | SiH <sub>4</sub> 150                                              |                                  |                                               |                          |                         |
|                                     | H <sub>2</sub> 300                                                | 300                              | 10                                            | 0.4                      | 20                      |
|                                     | SiH <sub>4</sub> 30                                               |                                  |                                               |                          |                         |
| 3rd layer region                    | CH <sub>4</sub> 300                                               | 300                              | 5                                             | 0.3                      | 0.5                     |
|                                     |                                                                   |                                  |                                               |                          |                         |

TABLE 147

| Order of lamination<br>(layer name) | Gases and their flow rates<br>(SCCM)                              | Substrate temperature<br>(°C.)   | RF discharging power<br>(mW/cm <sup>3</sup> ) | Inner pressure<br>(Torr) | Layer thickness<br>(μm) |
|-------------------------------------|-------------------------------------------------------------------|----------------------------------|-----------------------------------------------|--------------------------|-------------------------|
| Lower layer                         | GeH <sub>4</sub> 3                                                |                                  |                                               |                          |                         |
|                                     | B <sub>2</sub> H <sub>6</sub> (against SiH <sub>4</sub> ) 50 ppm  |                                  |                                               |                          |                         |
|                                     | NO 3                                                              |                                  |                                               |                          |                         |
|                                     | SiH <sub>4</sub> 25                                               |                                  |                                               |                          |                         |
|                                     | H <sub>2</sub> 5 → 100*                                           | 300                              | 0.5                                           | 0.2                      | 0.02                    |
|                                     | AlCl <sub>3</sub> /He<br>(S-side: 0.01 μm)                        | 100 → 15**<br>(UL-side: 0.01 μm) |                                               |                          |                         |
| Upper layer                         | SiH <sub>4</sub> 15 → 5**                                         |                                  |                                               |                          |                         |
|                                     | H <sub>2</sub> 60                                                 |                                  |                                               |                          |                         |
|                                     | B <sub>2</sub> H <sub>6</sub> (against SiH <sub>4</sub> ) 200 ppm |                                  |                                               |                          |                         |
|                                     | SiH <sub>4</sub> 300                                              | 300                              | 6                                             | 0.2                      | 10                      |
|                                     | H <sub>2</sub> 150                                                |                                  |                                               |                          |                         |
|                                     | SiH <sub>4</sub> 300                                              | 300                              | 10                                            | 0.4                      | 20                      |
| 1st layer region                    | SiH <sub>4</sub> 30                                               |                                  |                                               |                          |                         |
|                                     | CH <sub>4</sub> 300                                               | 300                              | 5                                             | 0.3                      | 0.5                     |
| 2nd layer region                    |                                                                   |                                  |                                               |                          |                         |
|                                     |                                                                   |                                  |                                               |                          |                         |
| 3rd layer region                    |                                                                   |                                  |                                               |                          |                         |
|                                     |                                                                   |                                  |                                               |                          |                         |

TABLE 148

| Order of lamination<br>(layer name) | Gases and<br>their flow rates<br>(SCCM)                                                                                                                                                                                                    | Substrate<br>temperature<br>(°C.)                                                                              | RF discharging<br>power<br>(mW/cm <sup>3</sup> ) | Inner<br>pressure<br>(Torr) | Layer<br>thickness<br>(μm) |
|-------------------------------------|--------------------------------------------------------------------------------------------------------------------------------------------------------------------------------------------------------------------------------------------|----------------------------------------------------------------------------------------------------------------|--------------------------------------------------|-----------------------------|----------------------------|
| Lower layer                         | GeH <sub>4</sub> 2<br>B <sub>2</sub> H <sub>6</sub> (against SiH <sub>4</sub> ) 50 ppm<br>NO 2<br>SiH <sub>4</sub> 20<br>H <sub>2</sub> 5 → 100*<br>AlCl <sub>3</sub> /He<br>(S-side: 0.01 μm)<br>(UL-side: 0.01 μm) 80 → 15**<br>15 → 5** | 300                                                                                                            | 0.3                                              | 0.2                         | 0.02                       |
| Upper layer                         | 1st<br>layer<br>region                                                                                                                                                                                                                     | SiH <sub>4</sub> 40<br>H <sub>2</sub> 200<br>B <sub>2</sub> H <sub>6</sub> (against SiH <sub>4</sub> ) 200 ppm | 300                                              | 5                           | 0.2                        |
|                                     | 2nd<br>layer<br>region                                                                                                                                                                                                                     | SiH <sub>4</sub> 100<br>H <sub>2</sub> 300                                                                     | 300                                              | 6                           | 0.3                        |
|                                     | 3rd<br>layer<br>region                                                                                                                                                                                                                     | SiH <sub>4</sub> 20<br>CH <sub>4</sub> 200                                                                     | 300                                              | 3                           | 0.2                        |

TABLE 149

| Order of lamination<br>(layer name) | Gases and<br>their flow rates<br>(SCCM)                                                                                                                                                                                                                                                                                                                           | Substrate<br>temperature<br>(°C.)                                                                                                                                        | RF discharging<br>power<br>(mW/cm <sup>3</sup> ) | Inner<br>pressure<br>(Torr) | Layer<br>thickness<br>(μm) |
|-------------------------------------|-------------------------------------------------------------------------------------------------------------------------------------------------------------------------------------------------------------------------------------------------------------------------------------------------------------------------------------------------------------------|--------------------------------------------------------------------------------------------------------------------------------------------------------------------------|--------------------------------------------------|-----------------------------|----------------------------|
| Lower layer                         | SiH <sub>4</sub> 50<br>GeH <sub>4</sub> 5<br>B <sub>2</sub> H <sub>6</sub> (against SiH <sub>4</sub> ) 100 ppm<br>NO 5<br>H <sub>2</sub> 5 → 200*<br>AlCl <sub>3</sub> /He 200 → 20**<br>SiH <sub>4</sub> 100<br>H <sub>2</sub> 1200<br>B <sub>2</sub> H <sub>6</sub> (against SiH <sub>4</sub> ) 200 ppm<br>(LL-side: 2 μm)<br>(U · 2nd · LR-side: 1 μm) 500 ppm | 500                                                                                                                                                                      | 5                                                | 0.4                         | 0.05                       |
| Upper layer                         | 1st<br>layer<br>region                                                                                                                                                                                                                                                                                                                                            | SiH <sub>4</sub> 100<br>H <sub>2</sub> 1200<br>B <sub>2</sub> H <sub>6</sub> (against SiH <sub>4</sub> ) 200 ppm<br>(LL-side: 2 μm)<br>(U · 2nd · LR-side: 1 μm) 500 ppm | 500                                              | 20                          | 0.4                        |
|                                     | 2nd<br>layer<br>region                                                                                                                                                                                                                                                                                                                                            | SiH <sub>4</sub> 300<br>H <sub>2</sub> 1500                                                                                                                              | 500                                              | 30                          | 0.5                        |
|                                     | 3rd<br>layer<br>region                                                                                                                                                                                                                                                                                                                                            | SiH <sub>4</sub> 200<br>C <sub>2</sub> H <sub>2</sub> 10 → 20*<br>NO 1                                                                                                   | 500                                              | 30                          | 0.4                        |

TABLE 150

| Order of lamination<br>(layer name) | Gases and<br>their flow rates<br>(SCCM)                                                                                                                                                                                                                                 | Substrate<br>temperature<br>(°C.)                                                                                                                                                                                                   | μW<br>discharging<br>power (mW/cm <sup>3</sup> ) | Inner<br>pressure<br>(Torr) | Layer<br>thickness<br>(μm) |
|-------------------------------------|-------------------------------------------------------------------------------------------------------------------------------------------------------------------------------------------------------------------------------------------------------------------------|-------------------------------------------------------------------------------------------------------------------------------------------------------------------------------------------------------------------------------------|--------------------------------------------------|-----------------------------|----------------------------|
| Lower layer                         | SiF <sub>4</sub> 10<br>GeH <sub>4</sub> 10<br>B <sub>2</sub> H <sub>6</sub> (against SiH <sub>4</sub> ) 50 ppm<br>NO 10<br>SiH <sub>4</sub> 150<br>H <sub>2</sub> 20 → 500*<br>AlCl <sub>3</sub> /He<br>(S-side: 0.01 μm)<br>(UL-side: 0.01 μm) 400 → 80**<br>80 → 50** | 250                                                                                                                                                                                                                                 | 0.5                                              | 0.6                         | 0.02                       |
| Upper layer                         | 1st<br>layer<br>region                                                                                                                                                                                                                                                  | SiH <sub>4</sub> 100<br>H <sub>2</sub> 500<br>B <sub>2</sub> H <sub>6</sub> (against SiH <sub>4</sub> ) 200 ppm<br>SiH <sub>4</sub> 700<br>SiF <sub>4</sub> 30<br>H <sub>2</sub> 500<br>SiH <sub>4</sub> 150<br>CH <sub>4</sub> 500 | 250                                              | 0.5                         | 0.5                        |
|                                     | 2nd<br>layer<br>region                                                                                                                                                                                                                                                  | SiF <sub>4</sub> 30<br>H <sub>2</sub> 500                                                                                                                                                                                           | 250                                              | 0.5                         | 20                         |
|                                     | 3rd<br>layer<br>region                                                                                                                                                                                                                                                  | SiH <sub>4</sub> 150<br>CH <sub>4</sub> 500                                                                                                                                                                                         | 250                                              | 0.5                         | 1                          |

TABLE 151

| Order of lamination (layer name) | Gases and their flow rates (SCCM)                                                                         | Substrate temperature (°C.) | RF discharging power (mW/cm <sup>3</sup> ) | Inner pressure (Torr) | Layer thickness (μm) |
|----------------------------------|-----------------------------------------------------------------------------------------------------------|-----------------------------|--------------------------------------------|-----------------------|----------------------|
| Lower layer                      | SiF <sub>4</sub>                                                                                          | 5                           |                                            |                       |                      |
|                                  | C <sub>2</sub> H <sub>2</sub>                                                                             | 10                          |                                            |                       |                      |
|                                  | B <sub>2</sub> H <sub>6</sub> (against SiH <sub>4</sub> )                                                 | 100 ppm                     | 250                                        | 5                     | 0.4                  |
|                                  | SiH <sub>4</sub>                                                                                          | 50                          |                                            |                       |                      |
|                                  | H <sub>2</sub>                                                                                            | 5 → 200*                    |                                            |                       |                      |
|                                  | AlCl <sub>3</sub> /He                                                                                     | 200 → 20**                  |                                            |                       |                      |
| Upper layer region               | 1st SiH <sub>4</sub>                                                                                      | 100                         |                                            |                       |                      |
|                                  | H <sub>2</sub>                                                                                            | 200                         |                                            |                       |                      |
|                                  | B <sub>2</sub> H <sub>6</sub> (against SiH <sub>4</sub> )<br>(LL-side: 3 μm)<br>(U · 2nd · LR-side: 2 μm) | 500 ppm                     | 250                                        | 10                    | 0.4                  |
|                                  |                                                                                                           | 500 → 0 ppm**               |                                            |                       |                      |
|                                  | AlCl <sub>3</sub> /He                                                                                     | 1 → 0**                     |                                            |                       |                      |
|                                  | SiH <sub>4</sub>                                                                                          | 200                         |                                            |                       |                      |
| 2nd layer region                 | C <sub>2</sub> H <sub>2</sub>                                                                             | 10 → 20*                    | 250                                        | 15                    | 0.4                  |
|                                  | NO                                                                                                        | 1                           |                                            |                       |                      |
|                                  |                                                                                                           |                             |                                            |                       |                      |
| 3rd layer region                 | SiH <sub>4</sub>                                                                                          | 300                         | 250                                        | 15                    | 0.5                  |
|                                  | H <sub>2</sub>                                                                                            | 300                         |                                            |                       | 10                   |

TABLE 152

| Order of lamination (layer name) | Gases and their flow rates (SCCM)                                                                         | Substrate temperature (°C.)      | RF discharging power (mW/cm <sup>3</sup> ) | Inner pressure (Torr) | Layer thickness (μm) |
|----------------------------------|-----------------------------------------------------------------------------------------------------------|----------------------------------|--------------------------------------------|-----------------------|----------------------|
| Lower layer                      | GeH <sub>4</sub>                                                                                          | 5                                |                                            |                       |                      |
|                                  | B <sub>2</sub> H <sub>6</sub> (against SiH <sub>4</sub> )                                                 | 100 ppm                          |                                            |                       |                      |
|                                  | NO                                                                                                        | 1                                |                                            |                       |                      |
|                                  | SiH <sub>4</sub>                                                                                          | 50                               |                                            |                       |                      |
|                                  | H <sub>2</sub>                                                                                            | 5 → 200*                         | 250                                        | 1                     | 0.4                  |
|                                  | AlCl <sub>3</sub> /He<br>(S-side: 0.01 μm)                                                                | 200 → 30**<br>(UL-side: 0.01 μm) |                                            |                       | 0.02                 |
| Upper layer region               | SiH <sub>4</sub>                                                                                          | 100                              |                                            |                       |                      |
|                                  | H <sub>2</sub>                                                                                            | 200                              |                                            |                       |                      |
|                                  | B <sub>2</sub> H <sub>6</sub> (against SiH <sub>4</sub> )<br>(LL-side: 8 μm)<br>(U · 2nd · LR-side: 2 μm) | 500 ppm                          | 250                                        | 10                    | 0.4                  |
|                                  |                                                                                                           | 500 → 0 ppm**                    |                                            |                       |                      |
|                                  | SiH <sub>4</sub>                                                                                          | 100                              |                                            |                       |                      |
|                                  | CH <sub>4</sub>                                                                                           | 100                              | 300                                        | 15                    | 0.4                  |
| 2nd layer region                 | SiH <sub>4</sub>                                                                                          | 300                              | 300                                        | 20                    | 0.5                  |
|                                  | H <sub>2</sub>                                                                                            | 300                              |                                            |                       |                      |
| 3rd layer region                 | SiH <sub>4</sub>                                                                                          | 50                               | 300                                        | 10                    | 0.4                  |
|                                  | CH <sub>4</sub>                                                                                           | 600                              |                                            |                       | 0.5                  |
| 4th layer region                 | SiH <sub>4</sub>                                                                                          |                                  |                                            |                       |                      |
|                                  | CH <sub>4</sub>                                                                                           |                                  |                                            |                       |                      |

TABLE 153

| Order of lamination (layer name) | Gases and their flow rates (SCCM)           | Substrate temperature (°C.)      | RF discharging power (mW/cm <sup>3</sup> ) | Inner pressure (Torr) | Layer thickness (μm) |
|----------------------------------|---------------------------------------------|----------------------------------|--------------------------------------------|-----------------------|----------------------|
| Lower layer                      | GeF <sub>4</sub>                            | 1 → 10*                          |                                            |                       |                      |
|                                  | NH <sub>3</sub>                             | 5 → 50*                          |                                            |                       |                      |
|                                  | SiH <sub>4</sub>                            | 10 → 100*                        |                                            |                       |                      |
|                                  | H <sub>2</sub>                              | 5 → 200*                         | 300                                        | 5                     | 0.4                  |
|                                  | AlCl <sub>3</sub> /He<br>(S-side: 0.05 μm)  | 200 → 40**<br>(UL-side: 0.15 μm) |                                            |                       | 0.2                  |
|                                  |                                             | 40 → 10**                        |                                            |                       |                      |
| Upper layer                      | SiH <sub>4</sub>                            | 100                              |                                            |                       |                      |
|                                  | H <sub>2</sub>                              | 500                              | 300                                        | 5                     | 0.4                  |
|                                  | PH <sub>3</sub> (against SiH <sub>4</sub> ) | 200 ppm                          |                                            |                       |                      |
|                                  | SiH <sub>4</sub>                            | 300                              | 300                                        | 15                    | 0.4                  |
|                                  | NH <sub>3</sub>                             | 50                               |                                            |                       | 25                   |
|                                  |                                             |                                  |                                            |                       |                      |
| 3rd layer region                 | SiH <sub>4</sub>                            | 100                              | 300                                        | 5                     | 0.2                  |
|                                  | H <sub>2</sub>                              | 300                              |                                            |                       | 8                    |
|                                  |                                             |                                  |                                            |                       |                      |
|                                  |                                             |                                  |                                            |                       |                      |
| 4th layer                        | SiH <sub>4</sub>                            | 100                              | 300                                        | 10                    | 0.4                  |
|                                  | NH <sub>3</sub>                             | 50                               |                                            |                       | 0.3                  |

TABLE 153-continued

| Order of lamination (layer name) | Gases and their flow rates (SCCM) | Substrate temperature (°C.) | RF discharging power (mW/cm <sup>3</sup> ) | Inner pressure (Torr) | Layer thickness (μm) |
|----------------------------------|-----------------------------------|-----------------------------|--------------------------------------------|-----------------------|----------------------|
| region                           |                                   |                             |                                            |                       |                      |

TABLE 154

| Order of lamination (layer name) | Gases and their flow rates (SCCM)                                                                                                                                                                                                                                                                                                     | Substrate temperature (°C.) | RF discharging power (mW/cm <sup>3</sup> ) | Inner pressure (Torr) | Layer thickness (μm) |
|----------------------------------|---------------------------------------------------------------------------------------------------------------------------------------------------------------------------------------------------------------------------------------------------------------------------------------------------------------------------------------|-----------------------------|--------------------------------------------|-----------------------|----------------------|
| Lower layer                      | PH <sub>3</sub> (against SiH <sub>4</sub> ) 50 ppm<br>NO 5 → 20*<br>SnH <sub>4</sub> 1 → 10*<br>SiH <sub>4</sub> 10 → 100*<br>H <sub>2</sub> 5 → 200*<br>AlCl <sub>3</sub> /He (S-side: 0.05 μm) 200 → 40**<br>(UL-side: 0.15 μm) 40 → 10**                                                                                           | 250                         | 5                                          | 0.4                   | 0.2                  |
| Upper layer                      | 1st layer region SiH <sub>4</sub> 100<br>H <sub>2</sub> 100<br>2nd layer region SiH <sub>4</sub> 100<br>CH <sub>4</sub> 100<br>3rd layer region PH <sub>3</sub> (against SiH <sub>4</sub> ) 50 ppm<br>SiH <sub>4</sub> 100<br>SiF <sub>4</sub> 5<br>4th layer region H <sub>2</sub> 200<br>SiH <sub>4</sub> 50<br>CH <sub>4</sub> 600 | 250 300 300 300             | 8 15 3 10                                  | 0.4 0.4 0.5 0.4       | 3 30 3 0.5           |
|                                  |                                                                                                                                                                                                                                                                                                                                       |                             |                                            |                       |                      |

TABLE 155

| Order of lamination (layer name) | Gases and their flow rates (SCCM)                                                                                                                                                                                                                                                                                                                                                   | Substrate temperature (°C.) | RF discharging power (mW/cm <sup>3</sup> ) | Inner pressure (Torr) | Layer thickness (μm) |
|----------------------------------|-------------------------------------------------------------------------------------------------------------------------------------------------------------------------------------------------------------------------------------------------------------------------------------------------------------------------------------------------------------------------------------|-----------------------------|--------------------------------------------|-----------------------|----------------------|
| Lower layer                      | GeF <sub>4</sub> 5<br>B <sub>2</sub> H <sub>6</sub> (against SiH <sub>4</sub> ) 100 ppm<br>SiH <sub>4</sub> 50<br>H <sub>2</sub> 5 → 200*<br>AlCl <sub>3</sub> /He 200 → 20**<br>SiH <sub>4</sub> 100<br>H <sub>2</sub> 200                                                                                                                                                         | 250                         | 5                                          | 0.4                   | 0.05                 |
| Upper layer                      | 1st layer region B <sub>2</sub> H <sub>6</sub> (against SiH <sub>4</sub> ) (LL-side: 2 μm) (U · 2nd · LR-side: 8 μm) 500 ppm<br>H <sub>2</sub> 500 → 0 ppm**<br>2nd layer region SiH <sub>4</sub> 300<br>C <sub>2</sub> H <sub>2</sub> 50<br>B <sub>2</sub> H <sub>6</sub> (against SiH <sub>4</sub> ) (U · 1st · LR-side: 1 μm) 0 → 100 ppm*<br>(U · 3rd · LR-side: 29 μm) 100 ppm | 250 330                     | 8 20                                       | 0.4 0.4               | 3 30                 |
|                                  |                                                                                                                                                                                                                                                                                                                                                                                     |                             |                                            |                       |                      |
|                                  | 3rd layer region Si <sub>24</sub> H <sub>6</sub> 200<br>H <sub>2</sub> 200                                                                                                                                                                                                                                                                                                          | 300                         | 10                                         | 0.5                   | 10                   |
|                                  | 4th layer region SiH <sub>4</sub> 200<br>C <sub>2</sub> H <sub>2</sub> 200                                                                                                                                                                                                                                                                                                          | 330                         | 10                                         | 0.4                   | 1                    |
|                                  |                                                                                                                                                                                                                                                                                                                                                                                     |                             |                                            |                       |                      |

TABLE 156

| Order of lamination (layer name) | Gases and their flow rates (SCCM)                                                                                                                                                                                                       | Substrate temperature (°C.) | RF discharging power (mW/cm <sup>3</sup> ) | Inner pressure (Torr) | Layer thickness (μm) |
|----------------------------------|-----------------------------------------------------------------------------------------------------------------------------------------------------------------------------------------------------------------------------------------|-----------------------------|--------------------------------------------|-----------------------|----------------------|
| Lower layer                      | SiH <sub>4</sub> 10 → 100*<br>PH <sub>3</sub> (against SiH <sub>4</sub> ) 50 ppm<br>NO 5 → 20*<br>GeH <sub>4</sub> 1 → 10*<br>SiF <sub>4</sub> 1 → 10*<br>H <sub>2</sub> 5 → 200*<br>AlCl <sub>3</sub> /He (S-side: 0.05 μm) 200 → 40** | 250                         | 5                                          | 0.4                   | 0.2                  |

TABLE 156-continued

| Order of lamination (layer name) | Gases and their flow rates (SCCM)                         |                  | Substrate temperature (°C.) | RF discharging power (mW/cm <sup>3</sup> ) | Inner pressure (Torr) | Layer thickness (μm) |
|----------------------------------|-----------------------------------------------------------|------------------|-----------------------------|--------------------------------------------|-----------------------|----------------------|
|                                  | (UL-side: 0.15 μm)                                        |                  | 40 → 10**                   |                                            |                       |                      |
| 1st layer region                 | SiH <sub>4</sub>                                          | 40               |                             |                                            |                       |                      |
|                                  | H <sub>2</sub>                                            | 200              |                             |                                            |                       |                      |
|                                  | PH <sub>3</sub> (against SiH <sub>4</sub> )               |                  |                             |                                            |                       |                      |
|                                  | (LL-side: 2 μm)                                           |                  | 250                         | 8                                          | 0.4                   | 3                    |
|                                  | (U - 2nd - LR-side: 1 μm)                                 |                  | 250 ppm                     |                                            |                       |                      |
| Upper layer                      | 2nd layer region                                          | SiH <sub>4</sub> | 300                         |                                            |                       |                      |
|                                  | NH <sub>3</sub>                                           | 30 → 50*         |                             |                                            |                       |                      |
|                                  | PH <sub>3</sub> (against SiH <sub>4</sub> )               | 50 ppm           |                             |                                            |                       |                      |
|                                  | 3rd layer region                                          | SiH <sub>4</sub> | 100                         |                                            |                       |                      |
|                                  | H <sub>2</sub>                                            | 300              |                             | 5                                          | 0.4                   | 8                    |
|                                  | 4th layer region                                          | SiH <sub>4</sub> | 100                         |                                            |                       |                      |
|                                  | NH <sub>3</sub>                                           | 80 → 100*        |                             | 5                                          | 0.4                   | 0.7                  |
|                                  | B <sub>2</sub> H <sub>6</sub> (against SiH <sub>4</sub> ) | 500 ppm          |                             |                                            |                       |                      |

TABLE 157

| Order of lamination (layer name) | Gases and their flow rates (SCCM)                         |          | Substrate temperature (°C.) | RF discharging power (mW/cm <sup>3</sup> ) | Inner pressure (Torr) | Layer thickness (μm) |
|----------------------------------|-----------------------------------------------------------|----------|-----------------------------|--------------------------------------------|-----------------------|----------------------|
| Lower layer                      | B <sub>2</sub> H <sub>6</sub> (against SiH <sub>4</sub> ) | 100 ppm  |                             |                                            |                       |                      |
|                                  | N <sub>2</sub>                                            | 100      |                             |                                            |                       |                      |
|                                  | GeH <sub>4</sub>                                          | 5        |                             |                                            |                       |                      |
|                                  | SiH <sub>4</sub>                                          | 50       | 250                         | 1                                          | 0.3                   | 0.02                 |
|                                  | H <sub>2</sub>                                            | 5 → 200* |                             |                                            |                       |                      |
| Upper layer                      | AlCl <sub>3</sub> /He                                     |          |                             |                                            |                       |                      |
|                                  | (S-side: 0.01 μm)                                         |          | 200 → 30**                  |                                            |                       |                      |
|                                  | (UL-side: 0.01 μm)                                        |          | 30 → 10**                   |                                            |                       |                      |
| 1st layer region                 | SiH <sub>4</sub>                                          | 100      |                             |                                            |                       |                      |
|                                  | He                                                        | 600      | 250                         | 10                                         | 0.4                   | 3                    |
|                                  | B <sub>2</sub> H <sub>6</sub> (against SiH <sub>4</sub> ) | 500 ppm  |                             |                                            |                       |                      |
| 2nd layer region                 | SiH <sub>4</sub>                                          | 300      |                             |                                            |                       |                      |
|                                  | B <sub>2</sub> H <sub>6</sub>                             | 0.5 ppm  | 250                         | 25                                         | 0.6                   | 25                   |
|                                  | H <sub>2</sub>                                            | 600      |                             |                                            |                       |                      |
| 3rd layer region                 | SiH <sub>4</sub>                                          | 50       |                             |                                            |                       |                      |
|                                  | CH <sub>4</sub>                                           | 500      | 250                         | 10                                         | 0.4                   | 1                    |

TABLE 158

| Order of lamination (layer name) | Gases and their flow rates (SCCM)                         |            | Substrate temperature (°C.) | RF discharging power (mW/cm <sup>3</sup> ) | Inner pressure (Torr) | Layer thickness (μm) |
|----------------------------------|-----------------------------------------------------------|------------|-----------------------------|--------------------------------------------|-----------------------|----------------------|
| Lower layer                      | SiH <sub>4</sub>                                          | 10 → 100*  |                             |                                            |                       |                      |
|                                  | GeH <sub>4</sub>                                          | 2 → 20*    |                             |                                            |                       |                      |
|                                  | SiF <sub>4</sub>                                          | 1 → 10*    |                             |                                            |                       |                      |
|                                  | NO                                                        | 5 → 20*    |                             |                                            |                       |                      |
|                                  | H <sub>2</sub>                                            | 5 → 200*   | 300                         | 10                                         | 0.4                   | 0.2                  |
| AlCl <sub>3</sub> /He            |                                                           |            |                             |                                            |                       |                      |
| (S-side: 0.05 μm)                |                                                           | 200 → 40** |                             |                                            |                       |                      |
|                                  | (UL-side 0.15 μm)                                         |            | 40 → 10**                   |                                            |                       |                      |
| 1st layer region                 | SiH <sub>4</sub>                                          | 100        |                             |                                            |                       |                      |
|                                  | H <sub>2</sub>                                            | 500        |                             |                                            |                       |                      |
|                                  | B <sub>2</sub> H <sub>6</sub> (against SiH <sub>4</sub> ) | 200 ppm    | 300                         | 8                                          | 0.4                   | 0.5                  |
| Upper layer                      | AlCl <sub>3</sub> /He                                     | 0.1        |                             |                                            |                       |                      |
| 2nd layer region                 | SiF <sub>4</sub>                                          | 0.5        |                             |                                            |                       |                      |
|                                  | SiH <sub>4</sub>                                          | 300        |                             |                                            |                       |                      |
|                                  | H <sub>2</sub>                                            | 500        |                             |                                            |                       |                      |
|                                  | CH <sub>4</sub>                                           | 1          |                             |                                            |                       |                      |
|                                  | AlCl <sub>3</sub> /He                                     | 0.1        | 300                         | 20                                         | 0.5                   | 20                   |
|                                  | NO                                                        | 0.1        |                             |                                            |                       |                      |
|                                  | SiF <sub>4</sub>                                          | 0.5        |                             |                                            |                       |                      |
| 3rd layer region                 | B <sub>2</sub> H <sub>6</sub> (against SiH <sub>4</sub> ) | 0.3 ppm    |                             |                                            |                       |                      |
|                                  | GeH <sub>4</sub>                                          | 0.1        |                             |                                            |                       |                      |
|                                  | SiH <sub>4</sub>                                          | 100        |                             |                                            |                       |                      |
|                                  | CH <sub>4</sub>                                           | 600        |                             |                                            |                       |                      |
|                                  | PH <sub>3</sub> (against SiH <sub>4</sub> )               | 3000 ppm   |                             |                                            |                       |                      |

TABLE 158-continued

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| 4th layer region                 | AlCl <sub>3</sub> /He 0.1                                         | 300                         | 15                                         | 0.4                   | 7                    |
|                                  | NO 0.1                                                            |                             |                                            |                       |                      |
|                                  | SiF <sub>4</sub> 0.5                                              |                             |                                            |                       |                      |
|                                  | B <sub>2</sub> H <sub>6</sub> (against SiH <sub>4</sub> ) 0.2 ppm |                             |                                            |                       |                      |
|                                  | GeH <sub>4</sub> 0.1                                              |                             |                                            |                       |                      |
|                                  | SiH <sub>4</sub> 40                                               |                             |                                            |                       |                      |
|                                  | CH <sub>4</sub> 600                                               |                             |                                            |                       |                      |
|                                  | AlCl <sub>3</sub> /He 0.1                                         |                             |                                            |                       |                      |
|                                  | NO 0.1                                                            |                             | 10                                         | 0.4                   | 0.1                  |
|                                  | SiF <sub>4</sub> 0.2                                              |                             |                                            |                       |                      |

TABLE 159

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 10 → 100*                                        | 300                         | 10                                         | 0.4                   | 0.2                  |
|                                  | GeH <sub>4</sub> 2 → 20*                                          |                             |                                            |                       |                      |
|                                  | SiF <sub>4</sub> 1 → 10*                                          |                             |                                            |                       |                      |
|                                  | NO 5 → 20*                                                        |                             |                                            |                       |                      |
|                                  | B <sub>2</sub> H <sub>6</sub> (against SiH <sub>4</sub> ) 100 ppm |                             |                                            |                       |                      |
|                                  | H <sub>2</sub> 5 → 200*                                           |                             |                                            |                       |                      |
|                                  | AlCl <sub>3</sub> /He (S-side: 0.05 μm)                           |                             |                                            |                       |                      |
|                                  | 200 → 40**                                                        |                             |                                            |                       |                      |
|                                  | (UL-side: 0.15 μm) 40 → 10**                                      |                             |                                            |                       |                      |
|                                  | SiH <sub>4</sub> 100                                              |                             |                                            |                       |                      |
| 1st layer region                 | H <sub>2</sub> 200                                                | 250                         | 8                                          | 0.4                   | 3                    |
|                                  | B <sub>2</sub> H <sub>6</sub> (against SiH <sub>4</sub> ) 500 ppm |                             |                                            |                       |                      |
|                                  | (LL-side: 2 μm) (U · 2nd · LR-side: 1 μm) 500 → 0 ppm**           |                             |                                            |                       |                      |
|                                  | AlCl <sub>3</sub> /He 0.1                                         |                             |                                            |                       |                      |
|                                  | SiF <sub>4</sub> 0.5                                              |                             |                                            |                       |                      |
|                                  | SiH <sub>4</sub> 100                                              |                             |                                            |                       |                      |
|                                  | SiF <sub>4</sub> 5                                                |                             |                                            |                       |                      |
|                                  | H <sub>2</sub> 200                                                |                             |                                            |                       |                      |
|                                  | B <sub>2</sub> H <sub>6</sub> (against SiH <sub>4</sub> ) 0.3 ppm |                             |                                            |                       |                      |
|                                  | NO 0.1                                                            |                             |                                            |                       |                      |
| Upper 2nd layer region           | CH <sub>4</sub> 1                                                 | 300                         | 3                                          | 0.5                   | 3                    |
|                                  | AlCl <sub>3</sub> /He 0.1                                         |                             |                                            |                       |                      |
|                                  | GeH <sub>4</sub> 0.1                                              |                             |                                            |                       |                      |
|                                  | SiH <sub>4</sub> 100                                              |                             |                                            |                       |                      |
|                                  | CH <sub>4</sub> 100                                               |                             |                                            |                       |                      |
|                                  | PH <sub>3</sub> (against SiH <sub>4</sub> ) 50 ppm                |                             |                                            |                       |                      |
|                                  | AlCl <sub>3</sub> /He 0.1                                         |                             |                                            |                       |                      |
|                                  | NO 0.1                                                            |                             |                                            |                       |                      |
|                                  | SiF <sub>4</sub> 0.5                                              |                             |                                            |                       |                      |
|                                  | B <sub>2</sub> H <sub>6</sub> 0.3 ppm                             |                             |                                            |                       |                      |
| 3rd layer region                 | GeH <sub>4</sub> 0.1                                              | 15                          | 0.4                                        | 30                    |                      |
|                                  | SiH <sub>4</sub> 100                                              |                             |                                            |                       |                      |
|                                  | CH <sub>4</sub> 100                                               |                             |                                            |                       |                      |
|                                  | PH <sub>3</sub> (against SiH <sub>4</sub> ) 50 ppm                |                             |                                            |                       |                      |
|                                  | AlCl <sub>3</sub> /He 0.1                                         |                             |                                            |                       |                      |
|                                  | NO 0.1                                                            |                             |                                            |                       |                      |
|                                  | SiF <sub>4</sub> 0.5                                              |                             |                                            |                       |                      |
|                                  | B <sub>2</sub> H <sub>6</sub> 0.3 ppm                             |                             |                                            |                       |                      |
|                                  | GeH <sub>4</sub> 0.1                                              |                             |                                            |                       |                      |
|                                  | SiH <sub>4</sub> 50                                               |                             |                                            |                       |                      |
| 4th layer region                 | CH <sub>4</sub> 600                                               | 10                          | 0.4                                        | 0.5                   |                      |
|                                  | AlCl <sub>3</sub> /He 0.1                                         |                             |                                            |                       |                      |
|                                  | SiF <sub>4</sub> 0.5                                              |                             |                                            |                       |                      |
|                                  | NO 0.1                                                            |                             |                                            |                       |                      |
|                                  | PH <sub>3</sub> (against SiH <sub>4</sub> ) 0.3 ppm               |                             |                                            |                       |                      |
|                                  | B <sub>2</sub> H <sub>6</sub> (against SiH <sub>4</sub> ) 0.3 ppm |                             |                                            |                       |                      |
|                                  | GeH <sub>4</sub> 0.1                                              |                             |                                            |                       |                      |
|                                  | SiH <sub>4</sub> 50                                               |                             |                                            |                       |                      |
|                                  | CH <sub>4</sub> 600                                               |                             |                                            |                       |                      |
|                                  | AlCl <sub>3</sub> /He 0.1                                         |                             |                                            |                       |                      |

TABLE 160

| Order of lamination (layer name) | Gases and their flow rates (SCCM)                  | Substrate temperature (°C.) | RF discharging power (mW/cm <sup>3</sup> ) | Inner pressure (Torr) | Layer thickness (μm) |
|----------------------------------|----------------------------------------------------|-----------------------------|--------------------------------------------|-----------------------|----------------------|
| Lower layer                      | SiH <sub>4</sub> 10 → 100*                         | 300                         | 10                                         | 0.4                   | 0.2                  |
|                                  | SiF <sub>4</sub> 1 → 10*                           |                             |                                            |                       |                      |
|                                  | NO 5 → 20*                                         |                             |                                            |                       |                      |
|                                  | GeH <sub>4</sub> 1 → 10*                           |                             |                                            |                       |                      |
|                                  | H <sub>2</sub> 5 → 200*                            |                             |                                            |                       |                      |
|                                  | AlCl <sub>3</sub> /He (S-side: 0.05 μm)            |                             |                                            |                       |                      |
|                                  | 200 → 40**                                         |                             |                                            |                       |                      |
|                                  | SiH <sub>4</sub> 100                               |                             |                                            |                       |                      |
|                                  | CH <sub>4</sub> 100                                |                             |                                            |                       |                      |
|                                  | PH <sub>3</sub> (against SiH <sub>4</sub> ) 50 ppm |                             |                                            |                       |                      |

TABLE 160-continued

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| (UL-side: 0.15 μm)               |                                                           |                             |                                            |                       |                      |
| Upper layer                      | H <sub>2</sub> S (against SiH <sub>4</sub> )              | 40 → 10**                   |                                            |                       |                      |
|                                  | SiH <sub>4</sub>                                          | 2 ppm                       |                                            |                       |                      |
|                                  | H <sub>2</sub>                                            | 100                         |                                            |                       |                      |
|                                  | B <sub>2</sub> H <sub>6</sub> (against SiH <sub>4</sub> ) | 500                         |                                            |                       |                      |
|                                  | SiF <sub>4</sub>                                          | 0.5                         |                                            |                       |                      |
|                                  | H <sub>2</sub> S (against SiH <sub>4</sub> )              | 1 ppm                       |                                            |                       |                      |
|                                  | AlCl <sub>3</sub> /He                                     | 0.1                         |                                            |                       |                      |
| 2nd layer region                 | SiH <sub>4</sub>                                          | 300                         |                                            |                       |                      |
|                                  | CH <sub>4</sub>                                           | 1                           |                                            |                       |                      |
|                                  | H <sub>2</sub>                                            | 500                         |                                            |                       |                      |
|                                  | B <sub>2</sub> H <sub>6</sub> (against SiH <sub>4</sub> ) | 0.3 ppm                     | 300                                        | 20                    | 0.5                  |
|                                  | GeH <sub>4</sub>                                          | 0.1                         |                                            |                       |                      |
|                                  | SiF <sub>4</sub>                                          | 0.5                         |                                            |                       |                      |
|                                  | NO                                                        | 0.1                         |                                            |                       |                      |
| 3rd layer region                 | H <sub>2</sub> S (against SiH <sub>4</sub> )              | 0.5 ppm                     |                                            |                       |                      |
|                                  | AlCl <sub>3</sub> /He                                     | 0.1                         |                                            |                       |                      |
|                                  | SiH <sub>4</sub>                                          | 100                         |                                            |                       |                      |
|                                  | CH <sub>4</sub>                                           | 600                         |                                            |                       |                      |
|                                  | GeH <sub>4</sub>                                          | 0.1                         |                                            |                       |                      |
|                                  | PH <sub>3</sub> (against SiH <sub>4</sub> )               | 3000 ppm                    |                                            |                       |                      |
|                                  | B <sub>2</sub> H <sub>6</sub> (against SiH <sub>4</sub> ) | 0.2 ppm                     | 300                                        | 15                    | 0.4                  |
| 4th layer region                 | SiF <sub>4</sub>                                          | 0.5                         |                                            |                       |                      |
|                                  | NO                                                        | 0.1                         |                                            |                       |                      |
|                                  | H <sub>2</sub> S (against SiH <sub>4</sub> )              | 1 ppm                       |                                            |                       |                      |
|                                  | AlCl <sub>3</sub> /He                                     | 0.1                         |                                            |                       |                      |
|                                  | SiH <sub>4</sub>                                          | 40                          |                                            |                       |                      |
|                                  | CH <sub>4</sub>                                           | 600                         |                                            |                       |                      |
|                                  | PH <sub>3</sub> (against SiH <sub>4</sub> )               | 1 ppm                       |                                            |                       |                      |
|                                  | B <sub>2</sub> H <sub>6</sub> (against SiH <sub>4</sub> ) | 0.1 ppm                     | 300                                        | 10                    | 0.4                  |
|                                  | H <sub>2</sub> S (against SiH <sub>4</sub> )              | 10 ppm                      |                                            |                       |                      |
|                                  | SiF <sub>4</sub>                                          | 0.2                         |                                            |                       |                      |
|                                  | NO                                                        | 0.1                         |                                            |                       |                      |
|                                  | AlCl <sub>3</sub> /He                                     | 0.1                         |                                            |                       |                      |
|                                  | GeH <sub>4</sub>                                          | 0.1                         |                                            |                       |                      |

TABLE 161

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Upper layer                      | SiH <sub>4</sub>                                          | 50                          |                                            |                       |                      |
|                                  | Mg(C <sub>5</sub> H <sub>5</sub> ) <sub>2</sub> /He       | 5                           |                                            |                       |                      |
|                                  | H <sub>2</sub>                                            | 10 → 200*                   |                                            |                       |                      |
|                                  | AlCl <sub>3</sub> /He                                     | 120 → 40**                  |                                            |                       |                      |
|                                  | SiH <sub>4</sub>                                          | 100                         |                                            |                       |                      |
|                                  | B <sub>2</sub> H <sub>6</sub> (against SiH <sub>4</sub> ) | 200 ppm                     | 250                                        | 8                     | 0.4                  |
|                                  | H <sub>2</sub>                                            | 500                         |                                            |                       |                      |
| Lower layer                      | SiH <sub>4</sub>                                          | 300                         |                                            |                       |                      |
|                                  | H <sub>2</sub>                                            | 300                         | 250                                        | 15                    | 0.5                  |
|                                  | SiH <sub>4</sub>                                          | 50                          |                                            |                       |                      |
|                                  | CH <sub>4</sub>                                           | 500                         | 250                                        | 10                    | 0.4                  |
|                                  | SiH <sub>4</sub>                                          | 50                          |                                            |                       |                      |
|                                  | CH <sub>4</sub>                                           | 500                         |                                            |                       |                      |

TABLE 162

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Upper layer                      | SiH <sub>4</sub>                                          | 50                          |                                            |                       |                      |
|                                  | AlCl <sub>3</sub> /He                                     | 120 → 40**                  | 250                                        | 5                     | 0.4                  |
|                                  | SiH <sub>4</sub>                                          | 100                         |                                            |                       |                      |
|                                  | B <sub>2</sub> H <sub>6</sub> (against SiH <sub>4</sub> ) | 200 ppm                     | 250                                        | 8                     | 0.4                  |
|                                  | H <sub>2</sub>                                            | 500                         |                                            |                       |                      |
|                                  | SiH <sub>4</sub>                                          | 300                         |                                            |                       |                      |
|                                  | H <sub>2</sub>                                            | 300                         | 250                                        | 15                    | 0.5                  |
| Lower layer                      | SiH <sub>4</sub>                                          | 50                          |                                            |                       |                      |
|                                  | CH <sub>4</sub>                                           | 500                         | 250                                        | 10                    | 0.4                  |
|                                  | SiH <sub>4</sub>                                          | 50                          |                                            |                       |                      |
|                                  | CH <sub>4</sub>                                           | 500                         |                                            |                       |                      |

TABLE 163

| Order of lamination (layer name) | Gases and their flow rates (SCCM)                                | Substrate temperature (°C.) | RF discharging power (mW/cm <sup>3</sup> ) | Inner pressure (Torr) | Layer thickness (μm) |
|----------------------------------|------------------------------------------------------------------|-----------------------------|--------------------------------------------|-----------------------|----------------------|
| Lower layer                      | SiH <sub>4</sub> 50                                              |                             |                                            |                       |                      |
|                                  | Mg(C <sub>5</sub> H <sub>5</sub> ) <sub>2</sub> /He 10           |                             |                                            |                       |                      |
|                                  | NO 5                                                             |                             |                                            |                       |                      |
|                                  | H <sub>2</sub> 10 → 200*                                         | 250                         | 5                                          | 0.4                   | 0.03                 |
|                                  | AlCl <sub>3</sub> /He (S-side: 0.01 μm)                          |                             |                                            |                       |                      |
| Upper layer                      |                                                                  | 100 → 10**                  |                                            |                       |                      |
|                                  | (UL-side: 0.02 μm) 10                                            |                             |                                            |                       |                      |
|                                  | B <sub>2</sub> H <sub>6</sub> (against SiH <sub>4</sub> ) 50 ppm |                             |                                            |                       |                      |
|                                  | 1st SiH <sub>4</sub> 100                                         |                             |                                            |                       |                      |
|                                  | H <sub>2</sub> 500                                               | 250                         | 8                                          | 0.4                   | 3                    |
|                                  | 2nd SiH <sub>4</sub> 300                                         |                             |                                            |                       |                      |
|                                  | H <sub>2</sub> 300                                               | 250                         | 15                                         | 0.5                   | 20                   |
|                                  | 3rd SiH <sub>4</sub> 50                                          |                             |                                            |                       |                      |
|                                  | CH <sub>4</sub> 500                                              | 250                         | 10                                         | 0.4                   | 0.5                  |
| region                           |                                                                  |                             |                                            |                       |                      |

TABLE 164

| Order of lamination (layer name) | Gases and their flow rates (SCCM)                                                 | Substrate temperature (°C.) | RF discharging power (mW/cm <sup>3</sup> ) | Inner pressure (Torr) | Layer thickness (μm) |
|----------------------------------|-----------------------------------------------------------------------------------|-----------------------------|--------------------------------------------|-----------------------|----------------------|
| Lower layer                      | SiH <sub>4</sub> 50                                                               |                             |                                            |                       |                      |
|                                  | B <sub>2</sub> H <sub>6</sub> (against SiH <sub>4</sub> ) 100 ppm                 |                             |                                            |                       |                      |
|                                  | Mg(C <sub>5</sub> H <sub>5</sub> ) <sub>2</sub> /He 8                             | 150                         | 0.5                                        |                       |                      |
|                                  | H <sub>2</sub> 5 → 200*                                                           | ↓                           | ↓                                          | 0.3                   | 0.02                 |
|                                  | AlCl <sub>3</sub> /He (S-side: 0.01 μm)                                           | 300                         | 1.5                                        |                       |                      |
| Upper layer                      |                                                                                   | 200 → 30**                  |                                            |                       |                      |
|                                  | (UL-side: 0.01 μm) 30 → 10**                                                      |                             |                                            |                       |                      |
|                                  | 1st SiH <sub>4</sub> 100                                                          |                             |                                            |                       |                      |
|                                  | H <sub>2</sub> 200                                                                |                             |                                            |                       |                      |
|                                  | B <sub>2</sub> H <sub>6</sub> (against SiH <sub>4</sub> ) 500 ppm (LL-side: 2 μm) | 250                         | 10                                         | 0.4                   | 3                    |
| 2nd layer                        | (U · 2nd · LR-side: 1 μm) 500 ppm → 0**                                           |                             |                                            |                       |                      |
|                                  | SiH <sub>4</sub> 300                                                              |                             |                                            |                       |                      |
|                                  | H <sub>2</sub> 500                                                                | 250                         | 20                                         | 0.5                   | 20                   |
| region                           |                                                                                   |                             |                                            |                       |                      |

TABLE 165

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 50                                               |                             |                                            |                       |                      |
|                                  | SiF <sub>4</sub> 5                                                |                             |                                            |                       |                      |
|                                  | Mg(C <sub>5</sub> H <sub>5</sub> ) <sub>2</sub> /He 5             |                             |                                            |                       |                      |
|                                  | B <sub>2</sub> H <sub>6</sub> (against SiH <sub>4</sub> ) 100 ppm | 250                         | 1                                          | 0.3                   | 0.02                 |
|                                  | H <sub>2</sub> 5 → 200*                                           |                             |                                            |                       |                      |
| 1st layer                        | AlCl <sub>3</sub> /He (S-side: 0.01 μm)                           |                             |                                            |                       |                      |
|                                  |                                                                   | 200 → 30**                  |                                            |                       |                      |
|                                  | (UL-side: 0.01 μm) 30 → 10**                                      |                             |                                            |                       |                      |
|                                  | N <sub>2</sub> 100                                                |                             |                                            |                       |                      |
|                                  | SiH <sub>4</sub> 100                                              |                             |                                            |                       |                      |
| Upper layer                      | He 600                                                            |                             |                                            |                       |                      |
|                                  | B <sub>2</sub> H <sub>6</sub> (against SiH <sub>4</sub> ) 500 ppm | 250                         | 10                                         | 0.4                   | 3                    |
|                                  | AlCl <sub>3</sub> /He 0.1                                         |                             |                                            |                       |                      |
|                                  | SiF <sub>4</sub> 0.5                                              |                             |                                            |                       |                      |
|                                  | Mg(C <sub>5</sub> H <sub>5</sub> ) <sub>2</sub> /He 0.1           |                             |                                            |                       |                      |
| 2nd layer                        | SiH <sub>4</sub> 300                                              |                             |                                            |                       |                      |
|                                  | He 600                                                            |                             |                                            |                       |                      |
|                                  | B <sub>2</sub> H <sub>6</sub> (against SiH <sub>4</sub> ) 0.3 ppm | 250                         | 25                                         | 0.6                   | 25                   |
|                                  | AlCl <sub>3</sub> /He 0.1                                         |                             |                                            |                       |                      |
|                                  | SiF <sub>4</sub> 0.5                                              |                             |                                            |                       |                      |
| 3rd layer                        | CH <sub>4</sub> 1                                                 |                             |                                            |                       |                      |
|                                  | NO 0.1                                                            |                             |                                            |                       |                      |
|                                  | Mg(C <sub>5</sub> H <sub>5</sub> ) <sub>2</sub> /He 0.1           |                             |                                            |                       |                      |
|                                  | SiH <sub>4</sub> 50                                               |                             |                                            |                       |                      |
|                                  | CH <sub>4</sub> 500                                               |                             |                                            |                       |                      |
| region                           |                                                                   |                             |                                            |                       |                      |

TABLE 165-continued

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| region                           | NO                                                        | 0.2                         | 250                                        | 10                    | 0.4                  |
|                                  | Mg(C <sub>5</sub> H <sub>5</sub> ) <sub>2</sub> /He       | 0.2                         |                                            |                       |                      |
|                                  | B <sub>2</sub> H <sub>6</sub> (against SiH <sub>4</sub> ) | 0.3 ppm                     |                                            |                       |                      |
|                                  | Al <sub>2</sub> Cl <sub>3</sub> /He                       | 0.2                         |                                            |                       |                      |
|                                  | SiF <sub>4</sub>                                          | 1                           |                                            |                       |                      |

TABLE 166

| Order of lamination (layer name) | Gases and their flow rates (SCCM)                                            | Substrate temperature (°C.) | RF discharging power (mW/cm <sup>3</sup> ) | Inner pressure (Torr) | Layer thickness (μm) |
|----------------------------------|------------------------------------------------------------------------------|-----------------------------|--------------------------------------------|-----------------------|----------------------|
| Lower layer                      | CH <sub>4</sub>                                                              | 50 → 200*                   | 250                                        | 10                    | 0.4                  |
|                                  | Mg(C <sub>5</sub> H <sub>5</sub> ) <sub>2</sub> /He                          | 1 → 10*                     |                                            |                       |                      |
|                                  | SiH <sub>4</sub>                                                             | 10 → 100*                   |                                            |                       |                      |
|                                  | H <sub>2</sub>                                                               | 5 → 200*                    |                                            |                       |                      |
|                                  | Al(CH <sub>3</sub> ) <sub>3</sub> /He<br>(S-side: 0.05 μm)                   | 200 → 40*                   |                                            |                       |                      |
| Upper layer region               | (UL-side: 0.15 μm)                                                           | 40 → 10*                    | 250                                        | 10                    | 0.2                  |
|                                  | SiH <sub>4</sub>                                                             | 100                         |                                            |                       |                      |
|                                  | H <sub>2</sub>                                                               | 200                         |                                            |                       |                      |
|                                  | B <sub>2</sub> H <sub>6</sub> (against SiH <sub>4</sub> )<br>(LL-side: 2 μm) | 500 ppm                     |                                            |                       |                      |
| 2nd layer region                 | (U + 2nd + LR-side: 1 μm)                                                    | 500 ppm → 0**               | 250                                        | 10                    | 0.4                  |
|                                  | SiH <sub>4</sub>                                                             | 400                         |                                            |                       |                      |
| 3rd layer region                 | Ar                                                                           | 200                         | 250                                        | 10                    | 0.5                  |
|                                  | SiH <sub>4</sub>                                                             | 100                         |                                            |                       |                      |
| region                           | NH <sub>3</sub>                                                              | 30                          | 250                                        | 5                     | 0.3                  |

TABLE 167

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | Mg(C <sub>5</sub> H <sub>5</sub> ) <sub>2</sub> /He       | 10                          | 300                                        | 10                    | 0.4                  |
|                                  | SiF <sub>4</sub>                                          | 1 → 10*                     |                                            |                       |                      |
|                                  | SiH <sub>4</sub>                                          | 10 → 100*                   |                                            |                       |                      |
|                                  | H <sub>2</sub>                                            | 5 → 200*                    |                                            |                       |                      |
|                                  | AlCl <sub>3</sub> /He<br>(S-side: 0.05 μm)                | 200 → 40**                  |                                            |                       |                      |
| Upper layer                      | (UL-side: 0.15 μm)                                        | 40 → 10**                   | 300                                        | 8                     | 0.5                  |
|                                  | SiH <sub>4</sub>                                          | 100                         |                                            |                       |                      |
|                                  | H <sub>2</sub>                                            | 500                         |                                            |                       |                      |
|                                  | B <sub>2</sub> H <sub>6</sub> (against SiH <sub>4</sub> ) | 200 ppm                     |                                            |                       |                      |
| 2nd layer region                 | SiH <sub>4</sub>                                          | 300                         | 20                                         | 0.5                   | 20                   |
|                                  | H <sub>2</sub>                                            | 500                         |                                            |                       |                      |
|                                  | SiH <sub>4</sub>                                          | 300                         |                                            |                       |                      |
|                                  | CH <sub>4</sub>                                           | 600                         |                                            |                       |                      |
| 3rd layer region                 | SiH <sub>4</sub>                                          | 100                         | 300                                        | 15                    | 0.4                  |
|                                  | CH <sub>4</sub>                                           | 600                         |                                            |                       |                      |
|                                  | PH <sub>3</sub> (against SiH <sub>4</sub> )               | 3000 ppm                    |                                            |                       |                      |
| 4th layer region                 | SiH <sub>4</sub>                                          | 40                          | 300                                        | 10                    | 0.4                  |
|                                  | CH <sub>4</sub>                                           | 600                         |                                            |                       |                      |

TABLE 168

| Order of lamination (layer name) | Gases and their flow rates (SCCM)                   | Substrate temperature (°C.) | RF discharging power (mW/cm <sup>3</sup> ) | Inner pressure (Torr) | Layer thickness (μm) |
|----------------------------------|-----------------------------------------------------|-----------------------------|--------------------------------------------|-----------------------|----------------------|
| Lower layer                      | SiH <sub>4</sub>                                    | 50                          | 330                                        | 5                     | 0.4                  |
|                                  | Mg(C <sub>5</sub> H <sub>5</sub> ) <sub>2</sub> /He | 5                           |                                            |                       |                      |
|                                  | PF <sub>5</sub> (against SiH <sub>4</sub> )         | 50 ppm                      |                                            |                       |                      |
|                                  | NO                                                  | 5                           |                                            |                       |                      |
|                                  | H <sub>2</sub>                                      | 5 → 200*                    |                                            |                       |                      |
| Upper layer                      | AlCl <sub>3</sub> /He                               | 200 → 20**                  | 330                                        | 8                     | 3                    |
|                                  | SiH <sub>4</sub>                                    | 100                         |                                            |                       |                      |
|                                  | H <sub>2</sub>                                      | 100                         |                                            |                       |                      |
|                                  | PF <sub>5</sub> (against SiH <sub>4</sub> )         | 100 ppm                     |                                            |                       |                      |

TABLE 168-continued

| Order of lamination (layer name) | Gases and their flow rates (SCCM)                                  | Substrate temperature (°C.) | RF discharging power (mW/cm <sup>3</sup> ) | Inner pressure (Torr) | Layer thickness (μm) |
|----------------------------------|--------------------------------------------------------------------|-----------------------------|--------------------------------------------|-----------------------|----------------------|
| 2nd layer region                 | SiH <sub>4</sub> 400                                               | 330                         | 25                                         | 0.5                   | 25                   |
|                                  | SiF <sub>4</sub> 10                                                |                             |                                            |                       |                      |
|                                  | H <sub>2</sub> 800                                                 |                             |                                            |                       |                      |
|                                  | SiH <sub>4</sub> 100                                               |                             |                                            |                       |                      |
|                                  | CH <sub>4</sub> 400                                                |                             |                                            |                       |                      |
| 3rd layer region                 | B <sub>2</sub> H <sub>6</sub> (against SiH <sub>4</sub> ) 5000 ppm | 350                         | 15                                         | 0.4                   | 5                    |
|                                  | SiH <sub>4</sub> 20                                                |                             |                                            |                       |                      |
|                                  | CH <sub>4</sub> 400                                                |                             |                                            |                       |                      |
| 4th layer region                 | B <sub>2</sub> H <sub>6</sub> (against SiH <sub>4</sub> ) 8000 ppm | 350                         | 10                                         | 0.4                   | 1                    |

TABLE 169

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 50                                               | 300                         | 1                                          | 0.3                   | 0.02                 |
|                                  | Mg(C <sub>5</sub> H <sub>5</sub> ) <sub>2</sub> /He 5             |                             |                                            |                       |                      |
|                                  | H <sub>2</sub> S (against SiH <sub>4</sub> ) 10 ppm               |                             |                                            |                       |                      |
|                                  | H <sub>2</sub> 5 → 200*                                           |                             |                                            |                       |                      |
|                                  | AlCl <sub>3</sub> /He (S-side: 0.01 μm) 200 → 30**                |                             |                                            |                       |                      |
| Upper layer                      | (UL-side: 0.01 μm) 30 → 10**                                      | 300                         | 8                                          | 0.4                   | 5                    |
|                                  | SiH <sub>4</sub> 100                                              |                             |                                            |                       |                      |
|                                  | H <sub>2</sub> 200                                                |                             |                                            |                       |                      |
|                                  | B <sub>2</sub> H <sub>6</sub> (against SiH <sub>4</sub> ) 200 ppm |                             |                                            |                       |                      |
|                                  | SiH <sub>4</sub> 300                                              |                             |                                            |                       |                      |
|                                  | H <sub>2</sub> 200                                                |                             |                                            |                       |                      |
|                                  | SiH <sub>4</sub> 50                                               |                             |                                            |                       |                      |
|                                  | N <sub>2</sub> 500                                                |                             |                                            |                       |                      |
| 4th layer region                 | PH <sub>3</sub> (against SiH <sub>4</sub> ) 3000 ppm              | 300                         | 20                                         | 0.4                   | 5                    |
|                                  | SiH <sub>4</sub> 40                                               |                             |                                            |                       |                      |
|                                  | CH <sub>4</sub> 600                                               |                             |                                            |                       |                      |
|                                  |                                                                   |                             |                                            |                       |                      |

TABLE 170

| Order of lamination (layer name) | Gases and their flow rates (SCCM)                                                 | Substrate temperature (°C.) | RF discharging power (mW/cm <sup>3</sup> ) | Inner pressure (Torr) | Layer thickness (μm) |
|----------------------------------|-----------------------------------------------------------------------------------|-----------------------------|--------------------------------------------|-----------------------|----------------------|
| Lower layer                      | SiH <sub>4</sub> 50                                                               | 300                         | 5                                          | 0.4                   | 0.05                 |
|                                  | B <sub>2</sub> H <sub>6</sub> (against SiH <sub>4</sub> ) 100 ppm                 |                             |                                            |                       |                      |
|                                  | C <sub>2</sub> H <sub>2</sub> 10                                                  |                             |                                            |                       |                      |
|                                  | NO 5                                                                              |                             |                                            |                       |                      |
|                                  | GeF <sub>4</sub> 5                                                                |                             |                                            |                       |                      |
|                                  | H <sub>2</sub> 5 → 200*                                                           |                             |                                            |                       |                      |
|                                  | AlCl <sub>3</sub> /He 200 → 20**                                                  |                             |                                            |                       |                      |
|                                  | Mg(C <sub>5</sub> H <sub>5</sub> ) <sub>2</sub> /He 8                             |                             |                                            |                       |                      |
|                                  | SiH <sub>4</sub> 100                                                              |                             |                                            |                       |                      |
|                                  | H <sub>2</sub> 200                                                                |                             |                                            |                       |                      |
| Upper layer                      | B <sub>2</sub> H <sub>6</sub> (against SiH <sub>4</sub> ) (LL-side: 3 μm) 500 ppm | 250                         | 10                                         | 0.4                   | 5                    |
|                                  | (U · 2nd · LR-side: 2 μm) 500 ppm → 0**                                           |                             |                                            |                       |                      |
|                                  | AlCl <sub>3</sub> /He 1 → 0**                                                     |                             |                                            |                       |                      |
|                                  | SiH <sub>4</sub> 300                                                              |                             |                                            |                       |                      |
|                                  | H <sub>2</sub> 300                                                                |                             |                                            |                       |                      |
| 2nd layer region                 | SiH <sub>4</sub> 100                                                              | 250                         | 15                                         | 0.5                   | 10                   |
|                                  | C <sub>2</sub> H <sub>2</sub> 10 → 20*                                            |                             |                                            |                       |                      |
|                                  | NO 1                                                                              |                             |                                            |                       |                      |
| 3rd layer region                 | SiH <sub>4</sub> 100                                                              | 250                         | 15                                         | 0.4                   | 20                   |
|                                  |                                                                                   |                             |                                            |                       |                      |

TABLE 171

| Order of lamination (layer name) | Gases and their flow rates (SCCM)                   | Substrate temperature (°C.) | RF discharging power (mW/cm <sup>3</sup> ) | Inner pressure (Torr) | Layer thickness (μm) |
|----------------------------------|-----------------------------------------------------|-----------------------------|--------------------------------------------|-----------------------|----------------------|
| Lower layer                      | SiH <sub>4</sub> 50                                 |                             |                                            |                       |                      |
|                                  | BF <sub>3</sub> (against SiH <sub>4</sub> ) 100 ppm |                             |                                            |                       |                      |
|                                  | NO 1                                                |                             |                                            |                       |                      |

TABLE 171-continued

| Order of lamination (layer name) | Gases and their flow rates (SCCM)                              | Substrate temperature (°C.) | RF discharging power (mW/cm <sup>3</sup> ) | Inner pressure (Torr) | Layer thickness (μm) |
|----------------------------------|----------------------------------------------------------------|-----------------------------|--------------------------------------------|-----------------------|----------------------|
| Upper layer region               | Mg(C <sub>5</sub> H <sub>5</sub> ) <sub>2</sub> /He            | 5                           |                                            |                       |                      |
|                                  | H <sub>2</sub>                                                 | 5 → 200*                    | 250                                        | 1                     | 0.4                  |
|                                  | AlCl <sub>3</sub> /He<br>(S-side: 0.01 μm)                     | 200 → 30**                  |                                            |                       |                      |
|                                  | (UL-side: 0.01 μm)                                             | 30 → 10**                   |                                            |                       |                      |
|                                  | SiH <sub>4</sub>                                               | 100                         |                                            |                       |                      |
|                                  | H <sub>2</sub>                                                 | 200                         |                                            |                       |                      |
|                                  | BF <sub>3</sub> (against SiH <sub>4</sub> )<br>(LL-side: 8 μm) | 250                         | 10                                         | 0.4                   | 10                   |
|                                  | (U + 2nd + LR-side: 2 μm)                                      | 500 ppm                     |                                            |                       |                      |
|                                  |                                                                | 500 ppm → 0**               |                                            |                       |                      |
|                                  | SiH <sub>4</sub>                                               | 300                         |                                            |                       |                      |
| 2nd layer region                 | H <sub>2</sub>                                                 | 300                         | 300                                        | 20                    | 0.5                  |
| 3rd layer region                 | SiH <sub>4</sub>                                               | 100                         | 300                                        | 15                    | 0.4                  |
| 4th layer region                 | CH <sub>3</sub>                                                | 100                         |                                            |                       | 20                   |
|                                  | SiH <sub>4</sub>                                               | 50                          | 300                                        | 10                    | 0.4                  |
|                                  | CH <sub>4</sub>                                                | 600                         |                                            |                       | 0.5                  |

TABLE 172

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 10 → 100*                   |                                            |                       |                      |
|                                  | Mg(C <sub>5</sub> H <sub>5</sub> ) <sub>2</sub> /He       |                             |                                            |                       |                      |
|                                  | NH <sub>3</sub>                                           | 5 → 50*                     |                                            |                       |                      |
|                                  | H <sub>2</sub>                                            | 5 → 200*                    |                                            |                       |                      |
|                                  | AlCl <sub>3</sub> /He<br>(S-side: 0.05 μm)                | 300                         | 5                                          | 0.4                   | 0.2                  |
|                                  | (UL-side: 0.15 μm)                                        | 200 → 40**                  |                                            |                       |                      |
|                                  |                                                           | 40 → 10**                   |                                            |                       |                      |
|                                  | SiF <sub>4</sub>                                          | 10                          |                                            |                       |                      |
|                                  | SiH <sub>4</sub>                                          | 100                         |                                            |                       |                      |
|                                  | H <sub>2</sub>                                            | 500                         | 300                                        | 5                     | 0.4                  |
| Upper layer                      | B <sub>2</sub> H <sub>6</sub> (against SiH <sub>4</sub> ) | 200 ppm                     |                                            |                       |                      |
|                                  | SiH <sub>4</sub>                                          | 100                         |                                            |                       |                      |
|                                  | H <sub>2</sub>                                            | 300                         | 300                                        | 5                     | 0.2                  |
|                                  |                                                           |                             |                                            |                       | 8                    |
|                                  | SiH <sub>4</sub>                                          | 300                         |                                            |                       |                      |
|                                  | NH <sub>3</sub>                                           | 50                          | 300                                        | 15                    | 0.4                  |
|                                  |                                                           |                             |                                            |                       | 25                   |
|                                  | SiH <sub>4</sub>                                          | 100                         | 300                                        | 10                    | 0.4                  |
|                                  | NH <sub>3</sub>                                           | 50                          |                                            |                       | 0.3                  |

TABLE 173

| Order of lamination (layer name) | Gases and their flow rates (SCCM)                                            | Substrate temperature (°C.) | RF discharging power (mW/cm <sup>3</sup> ) | Inner pressure (Torr) | Layer thickness (μm) |
|----------------------------------|------------------------------------------------------------------------------|-----------------------------|--------------------------------------------|-----------------------|----------------------|
| Lower layer                      | SiH <sub>4</sub>                                                             | 10 → 100*                   |                                            |                       |                      |
|                                  | SiF <sub>4</sub>                                                             | 1 → 5*                      |                                            |                       |                      |
|                                  | Mg(C <sub>5</sub> H <sub>5</sub> ) <sub>2</sub> /He                          | 10                          |                                            |                       |                      |
|                                  | H <sub>2</sub>                                                               | 5 → 200*                    | 250                                        | 5                     | 0.4                  |
|                                  | AlCl <sub>3</sub> /He<br>(S-side: 0.05 μm)                                   | 200 → 40**                  |                                            |                       |                      |
|                                  | (UL-side: 0.15 μm)                                                           | 40 → 10**                   |                                            |                       |                      |
|                                  | SiH <sub>4</sub>                                                             | 100                         |                                            |                       |                      |
|                                  | H <sub>2</sub>                                                               | 200                         |                                            |                       |                      |
|                                  | B <sub>2</sub> H <sub>6</sub> (against SiH <sub>4</sub> )<br>(LL-side: 2 μm) | 250                         | 8                                          | 0.4                   | 3                    |
|                                  | (U + 2nd + LR-side: 1 μm)                                                    | 500 ppm                     |                                            |                       |                      |
| Upper layer                      |                                                                              | 500 ppm → 0**               |                                            |                       |                      |
|                                  | SiH <sub>4</sub>                                                             | 100                         |                                            |                       |                      |
|                                  | SiF <sub>4</sub>                                                             | 5                           | 300                                        | 3                     | 0.5                  |
|                                  | H <sub>2</sub>                                                               | 200                         |                                            |                       |                      |
|                                  | SiH <sub>4</sub>                                                             | 100                         | 300                                        | 15                    | 0.4                  |
|                                  | CH <sub>3</sub>                                                              | 100                         |                                            |                       | 30                   |

TABLE 173-continued

| Order of lamination (layer name) | Gases and their flow rates (SCCM)                  | Substrate temperature (°C.) | RF discharging power (mW/cm <sup>3</sup> ) | Inner pressure (Torr) | Layer thickness (μm) |
|----------------------------------|----------------------------------------------------|-----------------------------|--------------------------------------------|-----------------------|----------------------|
| region                           | PH <sub>3</sub> (against SiH <sub>4</sub> ) 50 ppm |                             |                                            |                       |                      |
| 4th layer                        | SiH <sub>4</sub> 50                                |                             |                                            |                       |                      |
| region                           | CH <sub>4</sub> 600                                | 300                         | 10                                         | 0.4                   | 0.5                  |

TABLE 174

| Order of lamination (layer name) | Gases and their flow rates (SCCM)                             | Substrate temperature (°C.) | RF discharging power (mW/cm <sup>3</sup> ) | Inner pressure (Torr) | Layer thickness (μm) |
|----------------------------------|---------------------------------------------------------------|-----------------------------|--------------------------------------------|-----------------------|----------------------|
| Lower layer                      | SiH <sub>4</sub> 50                                           |                             |                                            |                       |                      |
|                                  | PH <sub>3</sub> (against SiH <sub>4</sub> ) 50 ppm            |                             |                                            |                       |                      |
|                                  | Si <sub>2</sub> F <sub>6</sub> 5                              | 250                         | 5                                          | 0.4                   | 0.05                 |
|                                  | Mg(C <sub>5</sub> H <sub>5</sub> ) <sub>2</sub> /He 8         |                             |                                            |                       |                      |
|                                  | H <sub>2</sub> 5 → 200*                                       |                             |                                            |                       |                      |
|                                  | AlCl <sub>3</sub> /He 200 → 20**                              |                             |                                            |                       |                      |
| Upper layer                      | SiH <sub>4</sub> 40                                           |                             |                                            |                       |                      |
| 1st region                       | H <sub>2</sub> 40                                             |                             |                                            |                       |                      |
|                                  | PH <sub>3</sub> (against SiH <sub>4</sub> ) 250 ppm           | 250                         | 8                                          | 0.4                   | 3                    |
|                                  | (LL-side: 2 μm)                                               |                             |                                            |                       |                      |
|                                  | (U · 2nd · LR-side: 1 μm)                                     |                             |                                            |                       |                      |
|                                  | 250 ppm → 0**                                                 |                             |                                            |                       |                      |
| 2nd layer region                 | Si <sub>2</sub> H <sub>6</sub> 200                            |                             |                                            |                       |                      |
|                                  | H <sub>2</sub> 200                                            | 300                         | 10                                         | 0.5                   | 10                   |
| 3rd layer region                 | SiH <sub>4</sub> 300                                          |                             |                                            |                       |                      |
|                                  | C <sub>2</sub> H <sub>2</sub> 50                              |                             |                                            |                       |                      |
| region                           | B <sub>2</sub> H <sub>6</sub> (against SiH <sub>4</sub> ) 330 |                             | 20                                         | 0.4                   | 30                   |
|                                  | (U · 2nd · LR-side: 1 μm)                                     |                             |                                            |                       |                      |
|                                  | 0 → 100 ppm*                                                  |                             |                                            |                       |                      |
|                                  | (U · 4th · LR-side: 29 μm)                                    |                             |                                            |                       |                      |
| 4th layer region                 | SiH <sub>4</sub> 100 ppm                                      |                             |                                            |                       |                      |
|                                  | C <sub>2</sub> H <sub>2</sub> 200                             | 330                         | 10                                         | 0.4                   | 1                    |

TABLE 175

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | Si <sub>2</sub> F <sub>6</sub> 1 → 5*                             |                             |                                            |                       |                      |
|                                  | B <sub>2</sub> H <sub>6</sub> (against SiH <sub>4</sub> ) 80 ppm  |                             |                                            |                       |                      |
|                                  | NH <sub>3</sub> 5                                                 |                             |                                            |                       |                      |
|                                  | Mg(C <sub>5</sub> H <sub>5</sub> ) <sub>2</sub> /He 1 → 8*        |                             |                                            |                       |                      |
|                                  | SiH <sub>4</sub> 10 → 100*                                        | 250                         | 5                                          | 0.4                   | 0.2                  |
|                                  | H <sub>2</sub> 5 → 200*                                           |                             |                                            |                       |                      |
|                                  | AlCl <sub>3</sub> /He (S-side: 0.05 μm) 200 → 40**                |                             |                                            |                       |                      |
|                                  | (UL-side: 0.15 μm) 40 → 10**                                      |                             |                                            |                       |                      |
| Upper layer                      | SiH <sub>4</sub> 100                                              |                             |                                            |                       |                      |
| 1st region                       | H <sub>2</sub> 500                                                | 300                         | 8                                          | 0.3                   | 3                    |
|                                  | B <sub>2</sub> H <sub>6</sub> (against SiH <sub>4</sub> ) 200 ppm |                             |                                            |                       |                      |
| 2nd region                       | SiH <sub>4</sub> 100                                              |                             |                                            |                       |                      |
|                                  | H <sub>2</sub> 300                                                | 300                         | 5                                          | 0.2                   | 8                    |
| 3rd layer region                 | SiH <sub>4</sub> 300                                              |                             |                                            |                       |                      |
|                                  | NH <sub>3</sub> 30 → 50*                                          | 300                         | 15                                         | 0.4                   | 25                   |
| 4th layer region                 | PH <sub>3</sub> (against SiH <sub>4</sub> ) 50 ppm                |                             |                                            |                       |                      |
|                                  | SiH <sub>4</sub> 100                                              |                             |                                            |                       |                      |
|                                  | NH <sub>3</sub> 80 → 100*                                         | 300                         | 5                                          | 0.4                   | 0.7                  |
|                                  | PH <sub>3</sub> (against SiH <sub>4</sub> ) 50 ppm                |                             |                                            |                       |                      |

TABLE 176

| Order of lamination (layer name) | Gases and their flow rates (SCCM)                     | Substrate temperature (°C.) | RF discharging power (mW/cm <sup>3</sup> ) | Inner pressure (Torr) | Layer thickness (μm) |
|----------------------------------|-------------------------------------------------------|-----------------------------|--------------------------------------------|-----------------------|----------------------|
| Lower layer                      | Mg(C <sub>5</sub> H <sub>5</sub> ) <sub>2</sub> /He 8 |                             |                                            |                       |                      |
|                                  | SiH <sub>4</sub> 50                                   |                             |                                            |                       |                      |
|                                  | H <sub>2</sub> 5 → 200*                               | 250                         | 1                                          | 0.4                   | 0.02                 |
|                                  | AlCl <sub>3</sub> /He                                 |                             |                                            |                       |                      |

TABLE 176-continued

| Order of lamination (layer name) | Gases and their flow rates (SCCM)           | Substrate temperature (°C.) | RF discharging power (mW/cm <sup>3</sup> ) | Inner pressure (Torr) | Layer thickness (μm) |
|----------------------------------|---------------------------------------------|-----------------------------|--------------------------------------------|-----------------------|----------------------|
| Upper layer region               | (S-side: 0.01 μm)                           | 200 → 30**                  |                                            |                       |                      |
|                                  | (UL-side: 0.01 μm)                          | 30 → 10**                   |                                            |                       |                      |
|                                  | 1st SiH <sub>4</sub>                        | 100                         |                                            |                       |                      |
|                                  | H <sub>2</sub>                              | 100                         | 300                                        | 8                     | 0.4                  |
|                                  | PH <sub>3</sub> (against SiH <sub>4</sub> ) | 100 ppm                     |                                            |                       |                      |
|                                  | 2nd SiH <sub>4</sub>                        | 300                         |                                            |                       |                      |
|                                  | H <sub>2</sub>                              | 500                         | 300                                        | 20                    | 0.5                  |
|                                  | 3rd SiH <sub>4</sub>                        | 100                         |                                            |                       |                      |
|                                  | GeH <sub>4</sub>                            | 10 → 50*                    | 300                                        | 5                     | 0.4                  |
|                                  | H <sub>2</sub>                              | 300                         |                                            |                       |                      |
| 4th layer region                 | SiH <sub>4</sub>                            | 100 → 40**                  |                                            |                       |                      |
|                                  | CH <sub>4</sub>                             | 100 → 600*                  | 300                                        | 10                    | 0.4                  |

TABLE 177

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | B <sub>2</sub> H <sub>6</sub> (against SiH <sub>4</sub> ) | 50 ppm                      |                                            |                       |                      |
|                                  | NO                                                        | 5                           |                                            |                       |                      |
|                                  | Mg(C <sub>5</sub> H <sub>5</sub> ) <sub>2</sub> /He       | 5                           |                                            |                       |                      |
|                                  | SiH <sub>4</sub>                                          | 50                          | 300                                        | 1                     | 0.3                  |
|                                  | H <sub>2</sub>                                            | 5 → 200*                    |                                            |                       |                      |
|                                  | <u>AlCl<sub>3</sub>/He</u>                                |                             |                                            |                       |                      |
|                                  | (S-side: 0.01 μm)                                         | 200 → 30**                  |                                            |                       |                      |
|                                  | (UL-side: 0.01 μm)                                        | 30 → 10**                   |                                            |                       |                      |
|                                  | 1st SiH <sub>4</sub>                                      | 100                         |                                            |                       |                      |
|                                  | H <sub>2</sub>                                            | 500                         | 300                                        | 8                     | 0.4                  |
| Upper layer                      | B <sub>2</sub> H <sub>6</sub> (against SiH <sub>4</sub> ) | 200 ppm                     |                                            |                       |                      |
|                                  | 2nd SiH <sub>4</sub>                                      | 300                         |                                            |                       |                      |
|                                  | H <sub>2</sub>                                            | 400                         | 300                                        | 15                    | 0.5                  |
|                                  | 3rd SiH <sub>4</sub>                                      | 50                          |                                            |                       |                      |
|                                  | CH <sub>4</sub>                                           | 500                         | 300                                        | 10                    | 0.4                  |
|                                  | region                                                    |                             |                                            |                       | 0.5                  |

TABLE 178

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | SiH <sub>4</sub>                                          | 50                          |                                            |                       |                      |
|                                  | Mg(C <sub>5</sub> H <sub>5</sub> ) <sub>2</sub> /He       | 5                           |                                            |                       |                      |
|                                  | B <sub>2</sub> H <sub>6</sub> (against SiH <sub>4</sub> ) | 50 ppm                      |                                            |                       |                      |
|                                  | NO                                                        | 5                           | 300                                        | 0.7                   | 0.3                  |
|                                  | H <sub>2</sub>                                            | 5 → 200*                    |                                            |                       |                      |
|                                  | <u>AlCl<sub>3</sub>/He</u>                                |                             |                                            |                       |                      |
|                                  | (S-side: 0.01 μm)                                         | 200 → 30**                  |                                            |                       |                      |
|                                  | (UL-side: 0.01 μm)                                        | 30 → 10**                   |                                            |                       |                      |
|                                  | 1st SiH <sub>4</sub>                                      | 80                          |                                            |                       |                      |
|                                  | H <sub>2</sub>                                            | 400                         | 300                                        | 7                     | 0.3                  |
| Upper layer                      | B <sub>2</sub> H <sub>6</sub> (against SiH <sub>4</sub> ) | 220 ppm                     |                                            |                       |                      |
|                                  | 2nd SiH <sub>4</sub>                                      | 200                         |                                            |                       |                      |
|                                  | H <sub>2</sub>                                            | 400                         | 300                                        | 12                    | 0.4                  |
|                                  | 3rd SiH <sub>4</sub>                                      | 40                          |                                            |                       |                      |
|                                  | CH <sub>4</sub>                                           | 400                         | 300                                        | 7                     | 0.3                  |
|                                  | region                                                    |                             |                                            |                       | 0.5                  |

TABLE 179

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | Mg(C <sub>5</sub> H <sub>5</sub> ) <sub>2</sub> /He       | 8                           |                                            |                       |                      |
|                                  | B <sub>2</sub> H <sub>6</sub> (against SiH <sub>4</sub> ) | 50 ppm                      |                                            |                       |                      |
|                                  | NO                                                        | 3                           |                                            |                       |                      |
|                                  | SiH <sub>4</sub>                                          | 25                          | 300                                        | 0.5                   | 0.2                  |
|                                  | H <sub>2</sub>                                            | 5 → 100*                    |                                            |                       |                      |
|                                  | <u>AlCl<sub>3</sub>/He</u>                                |                             |                                            |                       |                      |
|                                  | (S-side: 0.01 μm)                                         | 200 → 30**                  |                                            |                       |                      |
|                                  | (UL-side: 0.01 μm)                                        | 30 → 10**                   |                                            |                       |                      |
|                                  | 1st SiH <sub>4</sub>                                      | 100                         |                                            |                       |                      |
|                                  | H <sub>2</sub>                                            | 500                         | 300                                        | 10                    | 0.4                  |

TABLE 179-continued

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Upper layer                      | (S-side: 0.01 μm)<br>(UL-side: 0.01 μm) 100 → 15**                |                             |                                            |                       |                      |
|                                  | SiH <sub>4</sub> 60                                               |                             |                                            |                       |                      |
|                                  | H <sub>2</sub> 300                                                | 300                         | 6                                          | 0.2                   | 10                   |
|                                  | B <sub>2</sub> H <sub>6</sub> (against SiH <sub>4</sub> ) 220 ppm |                             |                                            |                       |                      |
|                                  | SiH <sub>4</sub> 150                                              |                             |                                            |                       |                      |
|                                  | H <sub>2</sub> 300                                                | 300                         | 10                                         | 0.4                   | 20                   |
| 3rd layer region                 | SiH <sub>4</sub> 30                                               |                             |                                            |                       |                      |
|                                  | CH <sub>4</sub> 300                                               | 300                         | 5                                          | 0.3                   | 0.5                  |

TABLE 180

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | Mg(C <sub>5</sub> H <sub>5</sub> ) <sub>2</sub> /He 10            |                             |                                            |                       |                      |
|                                  | B <sub>2</sub> H <sub>6</sub> (against SiH <sub>4</sub> ) 50 ppm  |                             |                                            |                       |                      |
|                                  | NO 2                                                              |                             |                                            |                       |                      |
|                                  | SiH <sub>4</sub> 20                                               | 300                         | 0.3                                        | 0.2                   | 0.02                 |
|                                  | H <sub>2</sub> 5 → 100*                                           |                             |                                            |                       |                      |
|                                  | AlCl <sub>3</sub> /He                                             |                             |                                            |                       |                      |
| Upper layer                      | (S-side: 0.01 μm) 80 → 15**                                       |                             |                                            |                       |                      |
|                                  | (UL-side: 0.01 μm) 15 → 5**                                       |                             |                                            |                       |                      |
|                                  | SiH <sub>4</sub> 40                                               |                             |                                            |                       |                      |
|                                  | H <sub>2</sub> 200                                                | 300                         | 5                                          | 0.2                   | 10                   |
|                                  | B <sub>2</sub> H <sub>6</sub> (against SiH <sub>4</sub> ) 220 ppm |                             |                                            |                       |                      |
|                                  | SiH <sub>4</sub> 100                                              |                             |                                            |                       |                      |
| 2nd layer region                 | H <sub>2</sub> 300                                                | 300                         | 6                                          | 0.3                   | 20                   |
|                                  | SiH <sub>4</sub> 20                                               |                             |                                            |                       |                      |
|                                  | CH <sub>4</sub> 200                                               | 300                         | 3                                          | 0.2                   | 0.5                  |
| 3rd layer region                 |                                                                   |                             |                                            |                       |                      |

TABLE 181

| Order of lamination (layer name) | Gases and their flow rates (SCCM)                                 | Substrate temperature (°C.) | RF discharging power (mW/cm <sup>3</sup> ) | Inner pressure (Torr) | Layer thickness (μm) |
|----------------------------------|-------------------------------------------------------------------|-----------------------------|--------------------------------------------|-----------------------|----------------------|
| Lower layer                      | SiH <sub>4</sub> 50                                               |                             |                                            |                       |                      |
|                                  | Mg(C <sub>5</sub> H <sub>5</sub> ) <sub>2</sub> /He 5             |                             |                                            |                       |                      |
|                                  | B <sub>2</sub> H <sub>6</sub> (against SiH <sub>4</sub> ) 100 ppm | 500                         | 5                                          | 0.4                   | 0.05                 |
|                                  | NO 5                                                              |                             |                                            |                       |                      |
|                                  | H <sub>2</sub> 5 → 200*                                           |                             |                                            |                       |                      |
|                                  | AlCl <sub>3</sub> /He 200 → 20**                                  |                             |                                            |                       |                      |
| 1st layer region                 | SiH <sub>4</sub> 100                                              |                             |                                            |                       |                      |
|                                  | H <sub>2</sub> 1200                                               | 500                         | 20                                         | 0.4                   | 3                    |
|                                  | B <sub>2</sub> H <sub>6</sub> (against SiH <sub>4</sub> )         |                             |                                            |                       |                      |
| 2nd layer region                 | (LL-side: 2 μm) 500 ppm                                           |                             |                                            |                       |                      |
|                                  | (U · 2nd · LR-side: 1 μm) 500 → 0 ppm**                           |                             |                                            |                       |                      |
|                                  | SiH <sub>4</sub> 300                                              |                             |                                            |                       |                      |
| 3rd layer region                 | H <sub>2</sub> 1500                                               | 500                         | 30                                         | 0.5                   | 10                   |
|                                  | SiH <sub>4</sub> 200                                              |                             |                                            |                       |                      |
|                                  | C <sub>2</sub> H <sub>2</sub> 10 → 20*                            | 500                         | 30                                         | 0.4                   | 20                   |
| NO                               | 1                                                                 |                             |                                            |                       |                      |

TABLE 182

| Order of lamination (layer name) | Gases and their flow rates (SCCM)                                | Substrate temperature (°C.) | μW discharging power (mW/cm <sup>3</sup> ) | Inner pressure (Torr) | Layer thickness (μm) |
|----------------------------------|------------------------------------------------------------------|-----------------------------|--------------------------------------------|-----------------------|----------------------|
| Lower layer                      | Si <sub>2</sub> F <sub>6</sub> 10                                |                             |                                            |                       |                      |
|                                  | Mg(C <sub>5</sub> H <sub>5</sub> ) <sub>2</sub> /He 10           |                             |                                            |                       |                      |
|                                  | B <sub>2</sub> H <sub>6</sub> (against SiH <sub>4</sub> ) 50 ppm |                             |                                            |                       |                      |
|                                  | NO 5                                                             |                             |                                            |                       |                      |
|                                  | SiH <sub>4</sub> 150                                             | 250                         | 0.5                                        | 0.6                   | 0.02                 |
|                                  | H <sub>2</sub> 20 → 500*                                         |                             |                                            |                       |                      |
| 1st layer                        | AlCl <sub>3</sub> /He                                            |                             |                                            |                       |                      |
|                                  | (S-side: 0.01 μm) 400 → 80**                                     |                             |                                            |                       |                      |
|                                  | (UL-side: 0.01 μm) 80 → 50**                                     |                             |                                            |                       |                      |
| Upper layer                      | SiH <sub>4</sub> 700                                             | 250                         | 0.5                                        | 0.5                   | 3                    |
|                                  | H <sub>2</sub> 500                                               |                             |                                            |                       |                      |

TABLE 182-continued

| Order of lamination (layer name) |        | Gases and their flow rates (SCCM)                         | Substrate temperature (°C.) | μW discharging power (mW/cm <sup>3</sup> ) | Inner pressure (Torr) | Layer thickness (μm) |
|----------------------------------|--------|-----------------------------------------------------------|-----------------------------|--------------------------------------------|-----------------------|----------------------|
| layer                            | region | B <sub>2</sub> H <sub>6</sub> (against SiH <sub>4</sub> ) | 200 ppm                     |                                            |                       |                      |
|                                  | 2nd    | SiH <sub>4</sub>                                          | 700                         |                                            |                       |                      |
|                                  | layer  | SiF <sub>4</sub>                                          | 30                          | 250                                        | 0.5                   | 0.5                  |
|                                  | region | H <sub>2</sub>                                            | 500                         |                                            |                       |                      |
|                                  | 3rd    | SiH <sub>4</sub>                                          | 150                         |                                            |                       |                      |
|                                  | layer  | CH <sub>4</sub>                                           | 300                         | 250                                        | 0.5                   | 1                    |
| region                           |        |                                                           |                             |                                            |                       |                      |

TABLE 183

| Order of lamination (layer name) |                                                           | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------------------------------------|-----------------------------|--------------------------------------------|-----------------------|----------------------|
| Lower layer                      | SiF <sub>4</sub>                                          | 5                                                         |                             |                                            |                       |                      |
|                                  | C <sub>2</sub> H <sub>2</sub>                             | 10                                                        |                             |                                            |                       |                      |
|                                  | B <sub>2</sub> H <sub>6</sub> (against SiH <sub>4</sub> ) | 100 ppm                                                   | 250                         | 5                                          | 0.4                   | 0.05                 |
|                                  | Mg(C <sub>5</sub> H <sub>5</sub> ) <sub>2</sub> /He       | 5                                                         |                             |                                            |                       |                      |
|                                  | H <sub>2</sub>                                            | 5 43 200*                                                 |                             |                                            |                       |                      |
|                                  | AlCl <sub>3</sub> /He                                     | 200 → 20**                                                |                             |                                            |                       |                      |
| Upper layer                      | 1st                                                       | SiH <sub>4</sub>                                          | 100                         |                                            |                       |                      |
|                                  | layer                                                     | H <sub>2</sub>                                            | 200                         |                                            |                       |                      |
|                                  | region                                                    | B <sub>2</sub> H <sub>6</sub> (against SiH <sub>4</sub> ) |                             | 250                                        | 10                    | 0.4                  |
|                                  |                                                           | (LL-side: 3 μm)                                           | 500 ppm                     |                                            |                       |                      |
|                                  |                                                           | (U · 2nd · LR-side: 2 μm)                                 | 500 → 0 ppm**               |                                            |                       |                      |
|                                  |                                                           | AlCl <sub>3</sub> /He                                     | 1 → **                      |                                            |                       |                      |
| 2nd                              | layer                                                     | SiH <sub>4</sub>                                          | 200                         |                                            |                       |                      |
|                                  | layer                                                     | C <sub>2</sub> H <sub>2</sub>                             | 10 → 20*                    | 250                                        | 15                    | 0.4                  |
|                                  | region                                                    | NO                                                        | 1                           |                                            |                       |                      |
|                                  | 3rd                                                       | SiH <sub>4</sub>                                          | 300                         |                                            |                       |                      |
|                                  | layer                                                     | H <sub>2</sub>                                            | 300                         | 250                                        | 15                    | 0.5                  |
|                                  | region                                                    |                                                           |                             |                                            |                       | 10                   |

TABLE 184

| Order of lamination (layer name) |                                                           | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------------------------------------|-----------------------------|--------------------------------------------|-----------------------|----------------------|
| Lower layer                      | Mg(C <sub>5</sub> H <sub>5</sub> ) <sub>2</sub> /He       | 5                                                         |                             |                                            |                       |                      |
|                                  | B <sub>2</sub> H <sub>6</sub> (against SiH <sub>4</sub> ) | 100 ppm                                                   |                             |                                            |                       |                      |
|                                  | NO                                                        | 1                                                         |                             |                                            |                       |                      |
|                                  | SiH <sub>4</sub>                                          | 50                                                        | 250                         | 1                                          | 0.4                   | 0.02                 |
|                                  | H <sub>2</sub>                                            | 5 → 200*                                                  |                             |                                            |                       |                      |
|                                  | AlCl <sub>3</sub> /He                                     |                                                           |                             |                                            |                       |                      |
| Upper layer                      | 1st                                                       | (S-side: 0.01 μm)                                         | 200 → 30**                  |                                            |                       |                      |
|                                  | layer                                                     | (UL-side: 0.01 μm)                                        | 30 → 10**                   |                                            |                       |                      |
|                                  | region                                                    | SiH <sub>4</sub>                                          | 100                         |                                            |                       |                      |
|                                  | 2nd                                                       | H <sub>2</sub>                                            | 200                         |                                            |                       |                      |
|                                  | layer                                                     | B <sub>2</sub> H <sub>6</sub> (against SiH <sub>4</sub> ) |                             | 250                                        | 10                    | 0.4                  |
|                                  | region                                                    | (LL-side: 8 μm)                                           | 500 ppm                     |                                            |                       |                      |
| 2nd                              | layer                                                     | (U · 2nd · LR-side: 2 μm)                                 | 500 → 0 ppm**               |                                            |                       |                      |
|                                  | layer                                                     | SiH <sub>4</sub>                                          | 100                         |                                            |                       |                      |
|                                  | region                                                    | CH <sub>4</sub>                                           | 100                         | 300                                        | 15                    | 0.4                  |
|                                  | 3rd                                                       | SiH <sub>4</sub>                                          | 300                         |                                            |                       |                      |
|                                  | layer                                                     | H <sub>2</sub>                                            | 300                         | 300                                        | 20                    | 0.5                  |
|                                  | region                                                    |                                                           |                             |                                            |                       | 5                    |
| 3rd                              | layer                                                     | SiH <sub>4</sub>                                          | 50                          |                                            |                       |                      |
|                                  | region                                                    | CH <sub>4</sub>                                           | 600                         | 300                                        | 10                    | 0.4                  |
|                                  | 4th                                                       | SiH <sub>4</sub>                                          |                             |                                            |                       |                      |
|                                  | layer                                                     | CH <sub>4</sub>                                           |                             |                                            |                       |                      |
|                                  | region                                                    |                                                           |                             |                                            |                       | 0.5                  |

TABLE 185

| Order of lamination (layer name) |                                                     | Gases and their flow rates (SCCM) | Substrate temperature (°C.) | RF discharging power (mW/cm <sup>3</sup> ) | Inner pressure (Torr) | Layer thickness (μm) |
|----------------------------------|-----------------------------------------------------|-----------------------------------|-----------------------------|--------------------------------------------|-----------------------|----------------------|
| Lower layer                      | Mg(C <sub>5</sub> H <sub>5</sub> ) <sub>2</sub> /He | 1 → 10*                           |                             |                                            |                       |                      |
|                                  | NH <sub>3</sub>                                     | 5 → 50*                           |                             |                                            |                       |                      |
|                                  | SiH <sub>4</sub>                                    | 10 → 100*                         |                             |                                            |                       |                      |
|                                  | H <sub>2</sub>                                      | 5 → 200*                          | 300                         | 5                                          | 0.4                   | 0.2                  |
|                                  | AlCl <sub>3</sub> /He                               |                                   |                             |                                            |                       |                      |
|                                  | 1st                                                 | (S-side: 0.05 μm)                 | 200 → 40**                  |                                            |                       |                      |
|                                  | layer                                               | (UL-side: 0.15 μm)                | 40 → 10**                   |                                            |                       |                      |
|                                  | region                                              | SiH <sub>4</sub>                  | 100                         |                                            |                       |                      |

TABLE 185-continued

| Order of lamination (layer name) | Gases and their flow rates (SCCM) |                                                           | Substrate temperature (°C.) | RF discharging power (mW/cm <sup>3</sup> ) | Inner pressure (Torr) | Layer thickness (μm) |
|----------------------------------|-----------------------------------|-----------------------------------------------------------|-----------------------------|--------------------------------------------|-----------------------|----------------------|
| Upper layer                      | layer region                      | H <sub>2</sub>                                            | 500                         | 300                                        | 5                     | 0.4                  |
|                                  | 2nd layer region                  | B <sub>2</sub> H <sub>6</sub> (against SiH <sub>4</sub> ) | 200 ppm                     |                                            |                       |                      |
|                                  | 3rd layer region                  | SiH <sub>4</sub>                                          | 300                         |                                            |                       |                      |
|                                  | 4th layer region                  | NH <sub>3</sub>                                           | 50                          | 300                                        | 15                    | 0.4                  |
|                                  | layer region                      | SiH <sub>4</sub>                                          | 100                         |                                            |                       | 25                   |
|                                  | layer region                      | H <sub>2</sub>                                            | 300                         |                                            | 5                     | 0.2                  |
| Lower layer                      | layer region                      | SiH <sub>4</sub>                                          | 100                         | 300                                        | 10                    | 0.8                  |
|                                  | layer region                      | NH <sub>3</sub>                                           | 50                          |                                            | 0.4                   | 0.3                  |

TABLE 186

| Order of lamination (layer name) | Gases and their flow rates (SCCM)                   |            | Substrate temperature (°C.) | RF discharging power (mW/cm <sup>3</sup> ) | Inner pressure (Torr) | Layer thickness (μm) |
|----------------------------------|-----------------------------------------------------|------------|-----------------------------|--------------------------------------------|-----------------------|----------------------|
| Lower layer                      | PH <sub>3</sub> (against SiH <sub>4</sub> )         | 50 ppm     |                             |                                            |                       |                      |
|                                  | NO (against SiH <sub>4</sub> )                      | 5 → 20*    |                             |                                            |                       |                      |
|                                  | Mg(C <sub>5</sub> H <sub>5</sub> ) <sub>2</sub> /He | 5 → 10*    |                             |                                            |                       |                      |
|                                  | SiH <sub>4</sub>                                    | 10 → 100*  | 250                         | 5                                          | 0.4                   | 0.2                  |
|                                  | H <sub>2</sub>                                      | 5 → 200*   |                             |                                            |                       |                      |
|                                  | <u>AlCl<sub>3</sub>/He</u>                          |            |                             |                                            |                       |                      |
| Upper layer                      | (S-side: 0.05 μm)                                   | 200 → 40** |                             |                                            |                       |                      |
|                                  | (UL-side: 0.15 μm)                                  | 40 → 10**  |                             |                                            |                       |                      |
|                                  | SiH <sub>4</sub>                                    | 100        |                             |                                            |                       |                      |
|                                  | H <sub>2</sub>                                      | 100        | 250                         | 8                                          | 0.4                   | 3                    |
|                                  | PH <sub>3</sub> (against SiH <sub>4</sub> )         | 100 ppm    |                             |                                            |                       |                      |
|                                  | SiH <sub>4</sub>                                    | 100        |                             |                                            |                       |                      |
| Lower layer                      | CH <sub>4</sub>                                     | 100        | 300                         | 15                                         | 0.4                   | 30                   |
|                                  | PH <sub>3</sub> (against SiH <sub>4</sub> )         | 50 ppm     |                             |                                            |                       |                      |
|                                  | SiF <sub>4</sub>                                    | 5          | 300                         | 3                                          | 0.5                   | 3                    |
|                                  | H <sub>2</sub>                                      | 200        |                             |                                            |                       |                      |
|                                  | SiH <sub>4</sub>                                    | 50         |                             |                                            |                       |                      |
|                                  | CH <sub>4</sub>                                     | 600        | 300                         | 10                                         | 0.4                   | 0.5                  |

TABLE 187

| Order of lamination (layer name) | Gases and their flow rates (SCCM)                           |               | Substrate temperature (°C.) | RF discharging power (mW/cm <sup>3</sup> ) | Inner pressure (Torr) | Layer thickness (μm) |
|----------------------------------|-------------------------------------------------------------|---------------|-----------------------------|--------------------------------------------|-----------------------|----------------------|
| Lower layer                      | Mg(C <sub>5</sub> H <sub>5</sub> ) <sub>2</sub> /He         | 5             |                             |                                            |                       |                      |
|                                  | B <sub>2</sub> H <sub>6</sub> (against SiH <sub>4</sub> )   | 100 ppm       |                             |                                            |                       |                      |
|                                  | SiH <sub>4</sub>                                            | 50            | 250                         | 5                                          | 0.4                   | 0.05                 |
|                                  | H <sub>2</sub>                                              | 5 → 200*      |                             |                                            |                       |                      |
|                                  | <u>AlCl<sub>3</sub>/He</u>                                  | 200 → 20**    |                             |                                            |                       |                      |
|                                  | N <sub>2</sub>                                              | 300           |                             |                                            |                       |                      |
| Upper layer                      | SiH <sub>4</sub>                                            | 100           |                             |                                            |                       |                      |
|                                  | H <sub>2</sub>                                              | 200           |                             |                                            |                       |                      |
|                                  | <u>B<sub>2</sub>H<sub>6</sub> (against SiH<sub>4</sub>)</u> |               | 250                         | 8                                          | 0.4                   | 3                    |
|                                  | (LL-side: 2 μm)                                             | 500 ppm       |                             |                                            |                       |                      |
|                                  | (U - 2nd · LR-side: 1 μm)                                   | 500 → 0 ppm** |                             |                                            |                       |                      |
|                                  | SiH <sub>4</sub>                                            | 300           |                             |                                            |                       |                      |
| Lower layer                      | C <sub>2</sub> H <sub>2</sub>                               | 50            |                             |                                            |                       |                      |
|                                  | <u>B<sub>2</sub>H<sub>6</sub> (against SiH<sub>4</sub>)</u> | 330           | 20                          | 0.4                                        | 30                    |                      |
|                                  | (U - 1st · LR-side: 1 μm)                                   | 0 → 100 ppm*  |                             |                                            |                       |                      |
|                                  | (U - 3rd · LR-side: 29 μm)                                  | 100 ppm       |                             |                                            |                       |                      |
|                                  | SiH <sub>4</sub>                                            | 200           |                             |                                            |                       |                      |
|                                  | H <sub>2</sub>                                              | 200           | 300                         | 10                                         | 0.5                   | 10                   |
| Upper layer                      | SiH <sub>4</sub>                                            | 200           |                             |                                            |                       |                      |
|                                  | C <sub>2</sub> H <sub>2</sub>                               | 200           | 330                         | 10                                         | 0.4                   | 1                    |

TABLE 188

| Order of lamination (layer name) | Gases and their flow rates (SCCM)           |           | Substrate temperature (°C.) | RF discharging power (mW/cm <sup>3</sup> ) | Inner pressure (Torr) | Layer thickness (μm) |
|----------------------------------|---------------------------------------------|-----------|-----------------------------|--------------------------------------------|-----------------------|----------------------|
| Lower layer                      | SiH <sub>4</sub>                            | 10 → 100* |                             |                                            |                       |                      |
|                                  | PH <sub>3</sub> (against SiH <sub>4</sub> ) | 50 ppm    |                             |                                            |                       |                      |
|                                  | NO                                          | 5 → 20*   |                             |                                            |                       |                      |

TABLE 188-continued

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Upper layer                      | Mg(C <sub>5</sub> H <sub>5</sub> ) <sub>2</sub> /He       | 1 → 8*                      | 250                                        | 5                     | 0.4                  |
|                                  | SiF <sub>4</sub>                                          | 1 → 10*                     |                                            |                       |                      |
|                                  | H <sub>2</sub>                                            | 5 → 200*                    |                                            |                       |                      |
|                                  | AlCl <sub>3</sub> /He                                     |                             |                                            |                       |                      |
|                                  | (S-side: 0.05 μm)                                         | 200 → 40**                  |                                            |                       |                      |
|                                  | (UL-side: 0.15 μm)                                        | 40 → 10**                   |                                            |                       |                      |
|                                  | SiH <sub>4</sub>                                          | 40                          |                                            |                       |                      |
|                                  | 1st layer region H <sub>2</sub>                           | 200                         | 250                                        | 8                     | 0.4                  |
|                                  | PH <sub>3</sub> (against SiH <sub>4</sub> )               |                             |                                            |                       | 3                    |
|                                  | (LL-side: 2 μm)                                           | 250 ppm                     |                                            |                       |                      |
| 2nd layer region                 | (U · 2nd · LR-side: 1 μm)                                 | 250 → 0 ppm**               |                                            |                       |                      |
|                                  | SiH <sub>4</sub>                                          | 300                         |                                            |                       |                      |
|                                  | C <sub>2</sub> H <sub>2</sub>                             | 50                          |                                            |                       |                      |
|                                  | B <sub>2</sub> H <sub>6</sub> (against SiH <sub>4</sub> ) | 330                         | 20                                         | 0.4                   | 30                   |
| 3rd layer region                 | (U · 1st · LR-side: 1 μm)                                 | 0 → 100 ppm*                |                                            |                       |                      |
|                                  | (U · 3rd · LR-side: 29 μm)                                | 100 ppm                     |                                            |                       |                      |
|                                  | SiH <sub>4</sub>                                          | 200                         | 300                                        | 10                    | 0.5                  |
| 4th layer region                 | H <sub>2</sub>                                            | 200                         |                                            |                       | 10                   |
|                                  | SiH <sub>4</sub>                                          | 200                         | 330                                        | 10                    | 0.4                  |
|                                  | C <sub>2</sub> H <sub>2</sub>                             | 200                         |                                            |                       | 1                    |

TABLE 189

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | B <sub>2</sub> H <sub>6</sub> (against SiH <sub>4</sub> ) | 100 ppm                     |                                            |                       |                      |
|                                  | Mg(C <sub>5</sub> H <sub>5</sub> ) <sub>2</sub> /He       | 5                           |                                            |                       |                      |
|                                  | SiH <sub>4</sub>                                          | 50                          |                                            |                       |                      |
|                                  | H <sub>2</sub>                                            | 5 → 200*                    | 250                                        | 1                     | 0.3                  |
|                                  | AlCl <sub>3</sub> /He                                     |                             |                                            |                       |                      |
|                                  | (S-side: 0.01 μm)                                         | 200 → 30**                  |                                            |                       |                      |
|                                  | (UL-side: 0.01 μm)                                        | 30 → 10**                   |                                            |                       |                      |
|                                  | 1st layer region SiH <sub>4</sub>                         | 100                         |                                            |                       |                      |
|                                  | He                                                        | 600                         | 250                                        | 10                    | 0.4                  |
|                                  | B <sub>2</sub> H <sub>6</sub> (against SiH <sub>4</sub> ) | 500 ppm                     |                                            |                       |                      |
| Upper layer                      | 2nd layer region SiH <sub>4</sub>                         | 300                         |                                            |                       |                      |
|                                  | 2nd layer region B <sub>2</sub> H <sub>6</sub>            | 0.5 ppm                     | 250                                        | 25                    | 0.6                  |
|                                  | 3rd layer region He                                       | 600                         |                                            |                       |                      |
|                                  | 3rd layer region SiH <sub>4</sub>                         | 50                          |                                            |                       |                      |
|                                  | 3rd layer region CH <sub>4</sub>                          | 500                         | 250                                        | 10                    | 0.4                  |
|                                  |                                                           |                             |                                            |                       | 1                    |

TABLE 190

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Lower layer                      | B <sub>2</sub> H <sub>6</sub> (against SiH <sub>4</sub> ) | 50 ppm*                     |                                            |                       |                      |
|                                  | SiH <sub>4</sub>                                          | 10 → 100*                   |                                            |                       |                      |
|                                  | GeH <sub>4</sub>                                          | 2 → 20*                     |                                            |                       |                      |
|                                  | SiF <sub>4</sub>                                          | 1 → 10*                     |                                            |                       |                      |
|                                  | Mg(C <sub>5</sub> H <sub>5</sub> ) <sub>2</sub> /He       | 1 → 10*                     | 300                                        | 10                    | 0.4                  |
|                                  | NO                                                        | 5 → 20*                     |                                            |                       |                      |
|                                  | H <sub>2</sub>                                            | 5 → 200*                    |                                            |                       |                      |
|                                  | AlCl <sub>3</sub> /He                                     |                             |                                            |                       |                      |
|                                  | (S-side: 0.05 μm)                                         | 200 → 40**                  |                                            |                       |                      |
|                                  | (UL-side: 0.15 μm)                                        | 40 → 10**                   |                                            |                       |                      |
| Upper layer                      | 1st layer region SiH <sub>4</sub>                         | 100                         |                                            |                       |                      |
|                                  | H <sub>2</sub>                                            | 500                         |                                            |                       |                      |
|                                  | Mg(C <sub>5</sub> H <sub>5</sub> ) <sub>2</sub> /He       | 0.2                         | 300                                        | 8                     | 0.4                  |
|                                  | B <sub>2</sub> H <sub>6</sub> (against SiH <sub>4</sub> ) | 200 ppm                     |                                            |                       |                      |
|                                  | AlCl <sub>3</sub> /He                                     | 0.2                         |                                            |                       |                      |
|                                  | SiF <sub>4</sub>                                          | 0.5                         |                                            |                       |                      |
|                                  | 2nd layer region SiH <sub>4</sub>                         | 300                         |                                            |                       |                      |
|                                  | H <sub>2</sub>                                            | 500                         |                                            |                       |                      |
|                                  | CH <sub>4</sub>                                           | 1                           |                                            |                       |                      |
|                                  | AlCl <sub>3</sub> /He                                     | 0.1                         | 300                                        | 20                    | 0.5                  |
|                                  | NO                                                        | 0.1                         |                                            |                       |                      |
|                                  | SiF <sub>4</sub>                                          | 0.5                         |                                            |                       |                      |
|                                  | B <sub>2</sub> H <sub>6</sub> (against SiH <sub>4</sub> ) | 0.3 ppm                     |                                            |                       |                      |
|                                  | Mg(C <sub>5</sub> H <sub>5</sub> ) <sub>2</sub> /He       | 0.1                         |                                            |                       |                      |
|                                  | SiH <sub>4</sub>                                          | 100                         |                                            |                       |                      |

TABLE 190-continued

| Order of lamination<br>(layer name) | Gases and<br>their flow rates<br>(SCCM)                   | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|-----------------------------------------------------------|-----------------------------------|--------------------------------------------------|-----------------------------|----------------------------|
| 4th<br>layer<br>region              | CH <sub>4</sub>                                           | 600                               |                                                  |                             |                            |
|                                     | PH <sub>3</sub> (against SiH <sub>4</sub> )               | 3000 ppm                          |                                                  |                             |                            |
|                                     | AlCl <sub>3</sub> /He                                     | 0.1                               | 300                                              | 15                          | 0.4                        |
|                                     | NO                                                        | 0.1                               |                                                  |                             |                            |
|                                     | SiF <sub>4</sub>                                          | 0.5                               |                                                  |                             |                            |
|                                     | B <sub>2</sub> H <sub>6</sub>                             | 0.2 ppm                           |                                                  |                             |                            |
|                                     | Mg(C <sub>5</sub> H <sub>5</sub> ) <sub>2</sub> /He       | 0.1                               |                                                  |                             |                            |
|                                     | SiH <sub>4</sub>                                          | 40                                |                                                  |                             |                            |
|                                     | CH <sub>4</sub>                                           | 600                               |                                                  |                             |                            |
|                                     | AlCl <sub>3</sub> /He                                     | 0.4                               | 300                                              | 10                          | 0.4                        |
| 4th<br>layer<br>region              | NO                                                        | 0.4                               |                                                  |                             | 0.1                        |
|                                     | SiF <sub>4</sub>                                          | 0.5                               |                                                  |                             |                            |
|                                     | B <sub>2</sub> H <sub>6</sub> (against SiH <sub>4</sub> ) | 1 ppm                             |                                                  |                             |                            |
|                                     | PH <sub>3</sub> (against SiH <sub>4</sub> )               | 1 ppm                             |                                                  |                             |                            |
|                                     | Mg(C <sub>5</sub> H <sub>5</sub> ) <sub>2</sub> /He       | 0.4                               |                                                  |                             |                            |

TABLE 191

| Order of lamination<br>(layer name) | Gases and<br>their flow rates<br>(SCCM)                   | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|-----------------------------------------------------------|-----------------------------------|--------------------------------------------------|-----------------------------|----------------------------|
| Lower layer                         | SiH <sub>4</sub>                                          | 10 → 100*                         |                                                  |                             |                            |
|                                     | SiF <sub>4</sub>                                          | 0.5                               |                                                  |                             |                            |
|                                     | NO                                                        | 0.1                               |                                                  |                             |                            |
|                                     | GeH <sub>4</sub>                                          | 1 → 10*                           |                                                  |                             |                            |
|                                     | CH <sub>4</sub>                                           | 2 → 20*                           |                                                  |                             |                            |
|                                     | H <sub>2</sub>                                            | 5 → 200*                          | 250                                              | 5                           | 0.4                        |
|                                     | AlCl <sub>3</sub> /He                                     |                                   |                                                  |                             | 0.2                        |
|                                     | (S-side: 0.05 μm)                                         | 200 → 40**                        |                                                  |                             |                            |
|                                     | (UL-side: 0.15 μm)                                        | 40 → 10**                         |                                                  |                             |                            |
|                                     | Mg(C <sub>5</sub> H <sub>5</sub> ) <sub>2</sub> /He       | 5                                 |                                                  |                             |                            |
| Upper layer                         | B <sub>2</sub> H <sub>6</sub> (against SiH <sub>4</sub> ) | 10 ppm                            |                                                  |                             |                            |
|                                     | SiH <sub>4</sub>                                          | 100                               |                                                  |                             |                            |
|                                     | H <sub>2</sub>                                            | 100                               |                                                  |                             |                            |
|                                     | B <sub>2</sub> H <sub>6</sub> (against SiH <sub>4</sub> ) | 600 → 0 ppm**                     | 250                                              | 10                          | 0.4                        |
|                                     | SiF <sub>4</sub>                                          | 10                                |                                                  |                             | 3                          |
|                                     | Mg(C <sub>5</sub> H <sub>5</sub> ) <sub>2</sub> /He       | 0.1                               |                                                  |                             |                            |
|                                     | AlCl <sub>3</sub> /He                                     | 0.1                               |                                                  |                             |                            |
|                                     | SiH <sub>4</sub>                                          | 100                               |                                                  |                             |                            |
|                                     | CH <sub>4</sub>                                           | 1                                 |                                                  |                             |                            |
|                                     | H <sub>2</sub>                                            | 200                               |                                                  |                             |                            |
| 3rd<br>layer<br>region              | B <sub>2</sub> H <sub>6</sub> (against SiH <sub>4</sub> ) | 0.3 ppm                           | 300                                              | 3                           | 0.5                        |
|                                     | GeH <sub>4</sub>                                          | 0.5                               |                                                  |                             |                            |
|                                     | SiF <sub>4</sub>                                          | 5                                 |                                                  |                             |                            |
|                                     | NO                                                        | 0.1                               |                                                  |                             |                            |
|                                     | Mg(C <sub>5</sub> H <sub>5</sub> ) <sub>2</sub> /He       | 0.1                               |                                                  |                             |                            |
|                                     | AlCl <sub>3</sub> /He                                     | 0.1                               |                                                  |                             |                            |
|                                     | SiH <sub>4</sub>                                          | 100                               |                                                  |                             |                            |
|                                     | CH <sub>4</sub>                                           | 100                               |                                                  |                             |                            |
|                                     | GeH <sub>4</sub>                                          | 0.1                               |                                                  |                             |                            |
|                                     | PH <sub>3</sub> (against SiH <sub>4</sub> )               | 50 ppm                            | 300                                              | 15                          | 0.4                        |
| 4th<br>layer<br>region              | B <sub>2</sub> H <sub>6</sub> (against SiH <sub>4</sub> ) | 0.3 ppm                           |                                                  |                             | 30                         |
|                                     | SiF <sub>4</sub>                                          | 5                                 |                                                  |                             |                            |
|                                     | NO                                                        | 0.1                               |                                                  |                             |                            |
|                                     | Mg(C <sub>5</sub> H <sub>5</sub> ) <sub>2</sub> /He       | 0.1                               |                                                  |                             |                            |
|                                     | AlCl <sub>3</sub> /He                                     | 0.1                               |                                                  |                             |                            |
|                                     | SiH <sub>4</sub>                                          | 50                                |                                                  |                             |                            |
|                                     | CH <sub>4</sub>                                           | 600                               |                                                  |                             |                            |
|                                     | PH <sub>3</sub> (against SiH <sub>4</sub> )               | 0.5 ppm                           | 300                                              | 10                          | 0.4                        |
|                                     | B <sub>2</sub> H <sub>6</sub> (against SiH <sub>4</sub> ) | 0.3 ppm                           |                                                  |                             | 0.5                        |
|                                     | Mg(C <sub>5</sub> H <sub>5</sub> ) <sub>2</sub> /He       | 0.1                               |                                                  |                             |                            |

TABLE 192

| Order of lamination<br>(layer name) | Gases and<br>their flow rates<br>(SCCM) | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|-----------------------------------------|-----------------------------------|--------------------------------------------------|-----------------------------|----------------------------|
| Lower layer                         | SiH <sub>4</sub>                        | 10 → 100*                         |                                                  |                             |                            |
|                                     | SiF <sub>4</sub>                        | 1 → 10*                           |                                                  |                             |                            |
|                                     | NO                                      | 5 → 20*                           |                                                  |                             |                            |
|                                     | H <sub>2</sub>                          | 5 → 200*                          |                                                  |                             |                            |

TABLE 192-continued

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Upper layer                      | <u>AlCl<sub>3</sub>/He</u>                                | 300                         | 10                                         | 0.4                   | 0.2                  |
|                                  | (S-side: 0.05 μm)                                         | 200 → 40**                  |                                            |                       |                      |
|                                  | (UL-side: 0.15 μm)                                        | 40 → 10**                   |                                            |                       |                      |
|                                  | Mg(C <sub>5</sub> H <sub>5</sub> ) <sub>2</sub> /He       | 10                          |                                            |                       |                      |
|                                  | H <sub>2</sub> S (against SiH <sub>4</sub> )              | 2 ppm                       |                                            |                       |                      |
|                                  | SiH <sub>4</sub>                                          | 100                         |                                            |                       |                      |
|                                  | H <sub>2</sub>                                            | 500                         |                                            |                       |                      |
|                                  | B <sub>2</sub> H <sub>6</sub> (against SiH <sub>4</sub> ) | 200 ppm                     |                                            |                       |                      |
|                                  | H <sub>2</sub> S (against SiH <sub>4</sub> )              | 1 ppm                       | 300                                        | 8                     | 0.4                  |
|                                  | SiF <sub>4</sub>                                          | 0.5                         |                                            |                       |                      |
|                                  | Mg(C <sub>5</sub> H <sub>5</sub> ) <sub>2</sub> /He       | 0.1                         |                                            |                       |                      |
|                                  | AlCl <sub>3</sub> /He                                     | 0.1                         |                                            |                       |                      |
|                                  | SiH <sub>4</sub>                                          | 300                         |                                            |                       |                      |
|                                  | CH <sub>4</sub>                                           | 1                           |                                            |                       |                      |
| Upper layer                      | H <sub>2</sub>                                            | 500                         |                                            |                       |                      |
|                                  | B <sub>2</sub> H <sub>6</sub> (against SiH <sub>4</sub> ) | 0.3 ppm                     |                                            |                       |                      |
|                                  | H <sub>2</sub> S (against SiH <sub>4</sub> )              | 0.5 ppm                     | 300                                        | 20                    | 0.5                  |
|                                  | SiF <sub>4</sub>                                          | 0.5                         |                                            |                       |                      |
|                                  | NO                                                        | 0.1                         |                                            |                       |                      |
|                                  | Mg(C <sub>5</sub> H <sub>5</sub> ) <sub>2</sub> /He       | 0.1                         |                                            |                       |                      |
|                                  | AlCl <sub>3</sub> /He                                     | 0.1                         |                                            |                       |                      |
|                                  | SiH <sub>4</sub>                                          | 100                         |                                            |                       |                      |
|                                  | CH <sub>4</sub>                                           | 600                         |                                            |                       |                      |
|                                  | H <sub>2</sub> S (against SiH <sub>4</sub> )              | 1 ppm                       |                                            |                       |                      |
|                                  | PH <sub>3</sub> (against SiH <sub>4</sub> )               | 3000 ppm                    |                                            |                       |                      |
|                                  | B <sub>2</sub> H <sub>6</sub> (against SiH <sub>4</sub> ) | 0.2 ppm                     | 300                                        | 15                    | 0.4                  |
|                                  | SiF <sub>4</sub>                                          | 0.5                         |                                            |                       |                      |
|                                  | NO                                                        | 0.1                         |                                            |                       |                      |
| Upper layer                      | Mg(C <sub>5</sub> H <sub>5</sub> ) <sub>2</sub> /He       | 0.1                         |                                            |                       |                      |
|                                  | AlCl <sub>3</sub> /He                                     | 0.1                         |                                            |                       |                      |
|                                  | SiH <sub>4</sub>                                          | 40                          |                                            |                       |                      |
|                                  | CH <sub>4</sub>                                           | 600                         |                                            |                       |                      |
|                                  | PH <sub>3</sub> (against SiH <sub>4</sub> )               | 1 ppm                       |                                            |                       |                      |
|                                  | B <sub>2</sub> H <sub>6</sub> (against SiH <sub>4</sub> ) | 0.1 ppm                     |                                            |                       |                      |
|                                  | Mg(C <sub>5</sub> H <sub>5</sub> ) <sub>2</sub> /He       | 0.1                         | 300                                        | 10                    | 0.4                  |
|                                  | SiF <sub>4</sub>                                          | 0.2                         |                                            |                       |                      |
|                                  | NO                                                        | 0.1                         |                                            |                       |                      |
|                                  | AlCl <sub>3</sub> /He                                     | 0.1                         |                                            |                       |                      |
|                                  | H <sub>2</sub> S (against SiH <sub>4</sub> )              | 10 ppm                      |                                            |                       |                      |

TABLE 193

| Order of lamination (layer name) | Gases and their flow rates (SCCM)                           | Substrate temperature (°C.) | RF discharging power (mW/cm <sup>3</sup> ) | Inner pressure (Torr) | Layer thickness (μm) |
|----------------------------------|-------------------------------------------------------------|-----------------------------|--------------------------------------------|-----------------------|----------------------|
| Upper layer                      | SiH <sub>4</sub>                                            | 20                          |                                            |                       |                      |
|                                  | H <sub>2</sub>                                              | 5 → 100*                    | 250                                        | 1                     | 0.01                 |
|                                  | Ar                                                          | 100                         |                                            |                       |                      |
|                                  | SiH <sub>4</sub>                                            | 100                         |                                            |                       |                      |
|                                  | <u>B<sub>2</sub>H<sub>6</sub> (against SiH<sub>4</sub>)</u> |                             |                                            |                       |                      |
|                                  | (LL-side: 8 μm)                                             | 500 ppm                     | 250                                        | 10                    | 0.4                  |
|                                  | (U · 2nd · LR-side: 2 μm)                                   | 500 → 0 ppm**               |                                            |                       |                      |
|                                  | H <sub>2</sub>                                              | 200                         |                                            |                       |                      |
|                                  | SiH <sub>4</sub>                                            | 100                         |                                            |                       |                      |
|                                  | CH <sub>4</sub>                                             | 100                         | 300                                        | 15                    | 0.4                  |
|                                  | SiH <sub>4</sub>                                            | 300                         | 300                                        | 20                    | 0.5                  |
|                                  | H <sub>2</sub>                                              | 300                         |                                            |                       |                      |
|                                  | SiH <sub>4</sub>                                            | 50                          | 300                                        | 10                    | 0.4                  |
|                                  | CH <sub>4</sub>                                             | 600                         |                                            |                       | 0.5                  |

TABLE 194

| Order of lamination (layer name) | Gases and their flow rates (SCCM)                                                 | Substrate temperature (°C.) | RF discharging power (mW/cm <sup>3</sup> ) | Inner pressure (Torr) | Layer thickness (μm) |
|----------------------------------|-----------------------------------------------------------------------------------|-----------------------------|--------------------------------------------|-----------------------|----------------------|
| Upper layer                      | SiH <sub>4</sub>                                                                  | 50                          |                                            |                       |                      |
|                                  | Cu(C <sub>4</sub> H <sub>7</sub> N <sub>2</sub> O <sub>2</sub> ) <sub>2</sub> /He | 5                           | 250                                        | 5                     | 0.4                  |
|                                  | H <sub>2</sub>                                                                    | 10 → 200*                   |                                            |                       |                      |
|                                  | AlCl <sub>3</sub> /He                                                             | 120 → 40**                  |                                            |                       |                      |
|                                  | SiH <sub>4</sub>                                                                  | 100                         |                                            |                       |                      |
|                                  | <u>B<sub>2</sub>H<sub>6</sub> (against SiH<sub>4</sub>)</u>                       | 200 ppm                     | 250                                        | 10                    | 0.4                  |
|                                  | H <sub>2</sub>                                                                    | 500                         |                                            |                       | 3                    |

TABLE 194-continued

| Order of lamination (layer name) | Gases and their flow rates (SCCM) |                  | Substrate temperature (°C.) | RF discharging power (mW/cm <sup>3</sup> ) | Inner pressure (Torr) | Layer thickness (μm) |
|----------------------------------|-----------------------------------|------------------|-----------------------------|--------------------------------------------|-----------------------|----------------------|
| layer region                     | 2nd layer                         | SiH <sub>4</sub> | 300                         |                                            |                       |                      |
|                                  |                                   | H <sub>2</sub>   | 300                         | 250                                        | 15                    | 0.5                  |
|                                  | 3rd layer                         | SiH <sub>4</sub> | 50                          |                                            |                       |                      |
|                                  |                                   | CH <sub>4</sub>  | 500                         | 250                                        | 10                    | 0.4                  |

TABLE 195

| Order of lamination (layer name) | Gases and their flow rates (SCCM) |                                                           | Substrate temperature (°C.) | RF discharging power (mW/cm <sup>3</sup> ) | Inner pressure (Torr) | Layer thickness (μm) |
|----------------------------------|-----------------------------------|-----------------------------------------------------------|-----------------------------|--------------------------------------------|-----------------------|----------------------|
| Upper layer region               | Lower layer                       | SiH <sub>4</sub>                                          | 50                          |                                            |                       |                      |
|                                  | 1st layer                         | AlCl <sub>3</sub> /He                                     | 120 → 40**                  | 250                                        | 5                     | 0.4                  |
|                                  |                                   | SiH <sub>4</sub>                                          | 100                         |                                            |                       |                      |
|                                  | 2nd layer                         | B <sub>2</sub> H <sub>6</sub> (against SiH <sub>4</sub> ) | 200 ppm                     | 250                                        | 10                    | 0.4                  |
|                                  |                                   | H <sub>2</sub>                                            | 500                         |                                            |                       |                      |
|                                  | 3rd layer                         | SiH <sub>4</sub>                                          | 300                         |                                            |                       |                      |
|                                  |                                   | H <sub>2</sub>                                            | 300                         | 250                                        | 15                    | 0.5                  |
|                                  | region                            | SiH <sub>4</sub>                                          | 50                          |                                            |                       |                      |
|                                  |                                   | CH <sub>4</sub>                                           | 500                         | 250                                        | 10                    | 0.4                  |

TABLE 196

| Order of lamination (layer name) | Gases and their flow rates (SCCM) |                                                                                   | Substrate temperature (°C.) | RF discharging power (mW/cm <sup>3</sup> ) | Inner pressure (Torr) | Layer thickness (μm) |
|----------------------------------|-----------------------------------|-----------------------------------------------------------------------------------|-----------------------------|--------------------------------------------|-----------------------|----------------------|
| Upper layer region               | Lower layer                       | SiH <sub>4</sub>                                                                  | 50                          |                                            |                       |                      |
|                                  |                                   | Cu(C <sub>4</sub> H <sub>7</sub> N <sub>2</sub> O <sub>2</sub> ) <sub>2</sub> /He | 10                          |                                            |                       |                      |
|                                  |                                   | H <sub>2</sub>                                                                    | 10 → 200*                   |                                            |                       |                      |
|                                  |                                   | AlCl <sub>3</sub> /He                                                             |                             | 250                                        | 5                     | 0.4                  |
|                                  |                                   | (S-side: 0.01 μm)                                                                 | 100 → 128                   |                                            |                       |                      |
|                                  |                                   |                                                                                   | 10**                        |                                            |                       |                      |
|                                  |                                   | (UL-side: 0.02 μm)                                                                | 10                          |                                            |                       |                      |
|                                  |                                   | B <sub>2</sub> H <sub>6</sub> (against SiH <sub>4</sub> )                         | 100 ppm                     |                                            |                       |                      |
|                                  | 1st layer                         | SiH <sub>4</sub>                                                                  | 100                         |                                            |                       |                      |
| Lower layer                      |                                   | H <sub>2</sub>                                                                    | 300                         | 250                                        | 10                    | 0.4                  |
|                                  |                                   | B <sub>2</sub> H <sub>6</sub> (against SiH <sub>4</sub> )                         | 200 ppm                     |                                            |                       |                      |
|                                  | 2nd layer                         | SiH <sub>4</sub>                                                                  | 300                         |                                            |                       |                      |
|                                  |                                   | H <sub>2</sub>                                                                    | 300                         | 250                                        | 15                    | 0.5                  |
| 2nd layer region                 | 3rd layer                         | SiH <sub>4</sub>                                                                  | 50                          |                                            |                       |                      |
|                                  |                                   | CH <sub>4</sub>                                                                   | 500                         | 250                                        | 10                    | 0.4                  |

TABLE 197

| Order of lamination (layer name) | Gases and their flow rates (SCCM) |                                                                                   | Substrate temperature (°C.) | RF discharging power (mW/cm <sup>3</sup> ) | Inner pressure (Torr) | Layer thickness (μm) |
|----------------------------------|-----------------------------------|-----------------------------------------------------------------------------------|-----------------------------|--------------------------------------------|-----------------------|----------------------|
| Upper layer region               | Lower layer                       | SiH <sub>4</sub>                                                                  | 50                          |                                            |                       |                      |
|                                  |                                   | Cu(C <sub>4</sub> H <sub>7</sub> N <sub>2</sub> O <sub>2</sub> ) <sub>2</sub> /He | 5 → 3**                     |                                            |                       |                      |
|                                  |                                   | Mg(C <sub>5</sub> H <sub>5</sub> ) <sub>2</sub> /He                               | 2                           | 150                                        | 0.5                   |                      |
|                                  |                                   | H <sub>2</sub>                                                                    | 5 → 200*                    | ↓                                          | ↓                     |                      |
|                                  |                                   | AlCl <sub>3</sub> /He                                                             |                             | 300                                        | 1.5                   |                      |
|                                  |                                   | (S-side: 0.01 μm)                                                                 | 200 → 30**                  |                                            |                       |                      |
|                                  |                                   | (UL-side: 0.01 μm)                                                                | 30 → 10**                   |                                            |                       |                      |
|                                  | 1st layer                         | SiH <sub>4</sub>                                                                  | 100                         |                                            |                       |                      |
|                                  |                                   | He                                                                                | 300                         |                                            |                       |                      |
| 2nd layer region                 |                                   | B <sub>2</sub> H <sub>6</sub> (against SiH <sub>4</sub> )                         |                             | 250                                        | 10                    | 0.4                  |
|                                  |                                   | (LL-side: 2 μm)                                                                   | 500 ppm                     |                                            |                       |                      |
|                                  |                                   | (U · 2nd · LR-side 1 μm)                                                          | 500 → 0 ppm**               |                                            |                       |                      |
| 2nd layer region                 | 2nd layer                         | SiH <sub>4</sub>                                                                  | 300                         | 250                                        | 20                    | 0.5                  |
|                                  |                                   | He                                                                                | 500                         |                                            |                       | 20                   |

TABLE 198

| Order of lamination<br>(layer name) | Gases and their flow rates<br>(SCCM)                                                  | Substrate temperature<br>(°C.) | RF discharging power<br>(mW/cm <sup>3</sup> ) | Inner pressure<br>(Torr) | Layer thickness<br>(μm) |
|-------------------------------------|---------------------------------------------------------------------------------------|--------------------------------|-----------------------------------------------|--------------------------|-------------------------|
| Lower layer                         | SiH <sub>4</sub> 50                                                                   |                                |                                               |                          |                         |
|                                     | B <sub>2</sub> H <sub>6</sub> (against SiH <sub>4</sub> ) 100 ppm                     |                                |                                               |                          |                         |
|                                     | Cu(C <sub>4</sub> H <sub>7</sub> N <sub>2</sub> O <sub>2</sub> ) <sub>2</sub> /He 6   |                                |                                               |                          |                         |
|                                     | Mg(C <sub>5</sub> H <sub>5</sub> ) <sub>2</sub> /He 3                                 |                                |                                               |                          |                         |
|                                     | H <sub>2</sub> 5 → 200*                                                               |                                |                                               |                          |                         |
|                                     | AlCl <sub>3</sub> /He<br>(S-side: 0.01 μm)                                            | 250                            | 1                                             | 0.3                      | 0.02                    |
|                                     | (UL-side: 0.01 μm)                                                                    | 200 → 30**                     |                                               |                          |                         |
|                                     | CH <sub>4</sub> 30 → 10**                                                             |                                |                                               |                          |                         |
|                                     | NO 1                                                                                  |                                |                                               |                          |                         |
|                                     | SiF <sub>4</sub> 8                                                                    |                                |                                               |                          |                         |
| Upper layer                         | SiH <sub>4</sub> 0.5                                                                  |                                |                                               |                          |                         |
|                                     | 1st layer region SiH <sub>4</sub> 100                                                 |                                |                                               |                          |                         |
|                                     | H <sub>2</sub> 300                                                                    |                                |                                               |                          |                         |
|                                     | B <sub>2</sub> H <sub>6</sub> (against SiH <sub>4</sub> ) 500 ppm                     |                                |                                               |                          |                         |
|                                     | Cu(C <sub>4</sub> H <sub>7</sub> N <sub>2</sub> O <sub>2</sub> ) <sub>2</sub> /He 0.4 | 250                            | 10                                            | 0.4                      | 3                       |
|                                     | Mg(C <sub>5</sub> H <sub>5</sub> ) <sub>2</sub> /He 0.3                               |                                |                                               |                          |                         |
|                                     | AlCl <sub>3</sub> /He 0.4                                                             |                                |                                               |                          |                         |
|                                     | SiF <sub>4</sub> 0.5                                                                  |                                |                                               |                          |                         |
|                                     | 2nd layer region SiH <sub>4</sub> 300                                                 |                                |                                               |                          |                         |
|                                     | H <sub>2</sub> 600                                                                    |                                |                                               |                          |                         |
| 3rd layer region                    | Cu(C <sub>4</sub> H <sub>7</sub> N <sub>2</sub> O <sub>2</sub> ) <sub>2</sub> /He 0.1 |                                |                                               |                          |                         |
|                                     | B <sub>2</sub> H <sub>6</sub> (against SiH <sub>4</sub> ) 0.3 ppm                     | 250                            | 25                                            | 0.6                      | 25                      |
|                                     | AlCl <sub>3</sub> /He 0.1                                                             |                                |                                               |                          |                         |
|                                     | SiF <sub>4</sub> 0.1                                                                  |                                |                                               |                          |                         |
|                                     | CH <sub>4</sub> 1                                                                     |                                |                                               |                          |                         |
|                                     | NO 0.1                                                                                |                                |                                               |                          |                         |
|                                     | Mg(C <sub>5</sub> H <sub>5</sub> ) <sub>2</sub> /He 0.2                               |                                |                                               |                          |                         |
|                                     | SiH <sub>4</sub> 50                                                                   |                                |                                               |                          |                         |
|                                     | CH <sub>4</sub> 500                                                                   |                                |                                               |                          |                         |
|                                     | Cu(C <sub>4</sub> H <sub>7</sub> N <sub>2</sub> O <sub>2</sub> ) <sub>2</sub> /He 1   |                                |                                               |                          |                         |
|                                     | No 1                                                                                  | 250                            | 10                                            | 0.4                      | 1                       |
|                                     | N <sub>2</sub> 1                                                                      |                                |                                               |                          |                         |
|                                     | B <sub>2</sub> H <sub>6</sub> (against SiH <sub>4</sub> ) 0.5 ppm                     |                                |                                               |                          |                         |
|                                     | Al <sub>2</sub> Cl <sub>5</sub> /He 1                                                 |                                |                                               |                          |                         |
|                                     | SiF <sub>4</sub> 2                                                                    |                                |                                               |                          |                         |
|                                     | Mg(C <sub>5</sub> H <sub>5</sub> ) <sub>2</sub> /He 1                                 |                                |                                               |                          |                         |

TABLE 199

| Order of lamination<br>(layer name) | Gases and their flow rates<br>(SCCM)                                                 | Substrate temperature<br>(°C.) | RF discharging power<br>(mW/cm <sup>3</sup> ) | Inner pressure<br>(Torr) | Layer thickness<br>(μm) |
|-------------------------------------|--------------------------------------------------------------------------------------|--------------------------------|-----------------------------------------------|--------------------------|-------------------------|
| Lower layer                         | SiF <sub>4</sub> 10                                                                  |                                |                                               |                          |                         |
|                                     | GeH <sub>4</sub> 1 → 5*                                                              |                                |                                               |                          |                         |
|                                     | SiH <sub>4</sub> 10 → 100*                                                           |                                |                                               |                          |                         |
|                                     | H <sub>2</sub> 5 → 200*                                                              |                                |                                               |                          |                         |
|                                     | AlCl <sub>3</sub> /He<br>(S-side: 0.05 μm)                                           | 250                            | 10                                            | 0.4                      | 0.2                     |
|                                     | (UL-side: 0.15 μm)                                                                   | 200 → 40**                     |                                               |                          |                         |
|                                     | 40 → 10**                                                                            |                                |                                               |                          |                         |
|                                     | B <sub>2</sub> H <sub>6</sub> (against SiH <sub>4</sub> ) 100 ppm                    |                                |                                               |                          |                         |
|                                     | Cu(C <sub>4</sub> H <sub>7</sub> N <sub>2</sub> O <sub>2</sub> ) <sub>2</sub> /He 20 |                                |                                               |                          |                         |
|                                     | SiH <sub>4</sub> 100                                                                 |                                |                                               |                          |                         |
| Upper layer                         | H <sub>2</sub> 200                                                                   |                                |                                               |                          |                         |
|                                     | B <sub>2</sub> H <sub>6</sub> (against SiH <sub>4</sub> ) 500 ppm                    | 250                            | 10                                            | 0.4                      | 3                       |
|                                     | (LL-side: 2 μm)                                                                      |                                |                                               |                          |                         |
|                                     | (U · 2nd · LR-side 1 μm)                                                             | 500 → 0 ppm**                  |                                               |                          |                         |
|                                     | SiF <sub>4</sub> 10                                                                  |                                |                                               |                          |                         |
|                                     | SiH <sub>4</sub> 400                                                                 |                                |                                               |                          |                         |
|                                     | Ar 200                                                                               | 250                            | 10                                            | 0.5                      | 15                      |
|                                     | SiF <sub>4</sub> 40                                                                  |                                |                                               |                          |                         |
|                                     | SiH <sub>4</sub> 100                                                                 |                                |                                               |                          |                         |
|                                     | NH <sub>3</sub> 30                                                                   | 250                            | 5                                             | 0.4                      | 0.3                     |
|                                     | SiF <sub>4</sub> 10                                                                  |                                |                                               |                          |                         |

TABLE 200

| Order of lamination<br>(layer name) | Gases and their flow rates<br>(SCCM)                                              | Substrate temperature<br>(°C.) | RF discharging power<br>(mW/cm <sup>3</sup> ) | Inner pressure<br>(Torr) | Layer thickness<br>(μm) |
|-------------------------------------|-----------------------------------------------------------------------------------|--------------------------------|-----------------------------------------------|--------------------------|-------------------------|
| Lower layer                         | CH <sub>4</sub> 5 → 25*                                                           |                                |                                               |                          |                         |
|                                     | Cu(C <sub>4</sub> H <sub>7</sub> N <sub>2</sub> O <sub>2</sub> ) <sub>2</sub> /He |                                |                                               |                          |                         |

TABLE 200-continued

| Order of lamination (layer name) | Gases and their flow rates (SCCM)                         | Substrate temperature (°C.) | RF discharging power (mW/cm <sup>3</sup> ) | Inner pressure (Torr) | Layer thickness (μm) |
|----------------------------------|-----------------------------------------------------------|-----------------------------|--------------------------------------------|-----------------------|----------------------|
| Upper layer                      | SiH <sub>4</sub>                                          | 1 → 10*                     |                                            |                       |                      |
|                                  | H <sub>2</sub>                                            | 10 → 100*                   |                                            |                       |                      |
|                                  | B <sub>2</sub> H <sub>6</sub> (against SiH <sub>4</sub> ) | 5 → 200*                    |                                            |                       |                      |
|                                  | AlCl <sub>3</sub> /He (S-side: 0.05 μm)                   | 10 ppm                      | 300                                        | 10                    | 0.4                  |
|                                  | (UL-side: 0.15 μm)                                        | 200 → 40**                  |                                            |                       |                      |
|                                  |                                                           | 40 → 10**                   |                                            |                       |                      |
|                                  | SiH <sub>4</sub>                                          | 100                         |                                            |                       |                      |
|                                  | H <sub>2</sub>                                            | 100                         | 300                                        | 10                    | 0.4                  |
|                                  | B <sub>2</sub> H <sub>6</sub> (against SiH <sub>4</sub> ) | 200 ppm                     |                                            |                       | 3                    |
|                                  | SiH <sub>4</sub>                                          | 300                         |                                            |                       |                      |
| 1st layer                        | H <sub>2</sub>                                            | 500                         | 300                                        | 20                    | 0.5                  |
| region                           | SiH <sub>4</sub>                                          | 100                         |                                            |                       |                      |
| 2nd layer                        | CH <sub>4</sub>                                           | 600                         | 300                                        | 15                    | 0.4                  |
| region                           | PH <sub>3</sub> (against SiH <sub>4</sub> )               | 3000 ppm                    |                                            |                       | 7                    |
| 3rd layer                        | SiH <sub>4</sub>                                          | 40                          |                                            |                       |                      |
| region                           | CH <sub>4</sub>                                           | 600                         | 300                                        | 10                    | 0.4                  |
| 4th layer                        |                                                           |                             |                                            |                       | 0.1                  |
| region                           |                                                           |                             |                                            |                       |                      |

TABLE 201

| Order of lamination (layer name) | Gases and their flow rates (SCCM)                                                 | Substrate temperature (°C.) | RF discharging power (mW/cm <sup>3</sup> ) | Inner pressure (Torr) | Layer thickness (μm) |
|----------------------------------|-----------------------------------------------------------------------------------|-----------------------------|--------------------------------------------|-----------------------|----------------------|
| Upper layer                      | SiH <sub>4</sub>                                                                  | 50                          |                                            |                       |                      |
|                                  | Cu(C <sub>4</sub> H <sub>7</sub> N <sub>2</sub> O <sub>2</sub> ) <sub>2</sub> /He | 10                          |                                            |                       |                      |
|                                  | Mg(C <sub>5</sub> H <sub>5</sub> ) <sub>2</sub> /He                               | 3                           | 330                                        | 5                     | 0.4                  |
|                                  | H <sub>2</sub>                                                                    | 5 → 200*                    |                                            |                       |                      |
|                                  | AlCl <sub>3</sub> /He                                                             | 200 → 20**                  |                                            |                       |                      |
|                                  | SiH <sub>4</sub>                                                                  | 100                         |                                            |                       |                      |
|                                  | H <sub>2</sub>                                                                    | 300                         | 330                                        | 10                    | 0.4                  |
|                                  | PH <sub>3</sub> (against SiH <sub>4</sub> )                                       | 100 ppm                     |                                            |                       | 3                    |
|                                  | SiH <sub>4</sub>                                                                  | 400                         |                                            |                       |                      |
|                                  | SiF <sub>4</sub>                                                                  | 10                          | 330                                        | 25                    | 0.5                  |
| 1st layer                        | H <sub>2</sub>                                                                    | 800                         |                                            |                       | 25                   |
| region                           | SiH <sub>4</sub>                                                                  | 100                         |                                            |                       |                      |
| 2nd layer                        | CH <sub>4</sub>                                                                   | 400                         | 350                                        | 15                    | 0.4                  |
| region                           | B <sub>2</sub> H <sub>6</sub> (against SiH <sub>4</sub> )                         | 5000 ppm                    |                                            |                       | 5                    |
| 3rd layer                        | SiH <sub>4</sub>                                                                  | 20                          |                                            |                       |                      |
| region                           | CH <sub>4</sub>                                                                   | 400                         | 350                                        | 10                    | 0.4                  |
| 4th layer                        | B <sub>2</sub> H <sub>6</sub> (against SiH <sub>4</sub> )                         | 8000 ppm                    |                                            |                       | 1                    |
| region                           |                                                                                   |                             |                                            |                       |                      |

TABLE 202

| Order of lamination (layer name) | Gases and their flow rates (SCCM)                                                 | Substrate temperature (°C.) | RF discharging power (mW/cm <sup>3</sup> ) | Inner pressure (Torr) | Layer thickness (μm) |
|----------------------------------|-----------------------------------------------------------------------------------|-----------------------------|--------------------------------------------|-----------------------|----------------------|
| Upper layer                      | SiH <sub>4</sub>                                                                  | 50                          |                                            |                       |                      |
|                                  | Cu(C <sub>4</sub> H <sub>7</sub> N <sub>2</sub> O <sub>2</sub> ) <sub>2</sub> /He | 30                          |                                            |                       |                      |
|                                  | Mg(C <sub>5</sub> H <sub>5</sub> ) <sub>2</sub> /He                               | 2                           |                                            |                       |                      |
|                                  | H <sub>2</sub>                                                                    | 5 → 200*                    | 300                                        | 1                     | 0.3                  |
|                                  | AlCl <sub>3</sub> /He (S-side: 0.01 μm)                                           | 200 → 30**                  |                                            |                       |                      |
|                                  | (UL-side: 0.01 μm)                                                                | 30 → 10**                   |                                            |                       |                      |
|                                  | SiH <sub>4</sub>                                                                  | 100                         |                                            |                       |                      |
|                                  | H <sub>2</sub>                                                                    | 500                         | 300                                        | 10                    | 0.4                  |
|                                  | B <sub>2</sub> H <sub>6</sub> (against SiH <sub>4</sub> )                         | 200 ppm                     |                                            |                       | 3                    |
|                                  | SiH <sub>4</sub>                                                                  | 300                         |                                            |                       |                      |
| 1st layer                        | H <sub>2</sub>                                                                    | 200                         | 300                                        | 20                    | 0.5                  |
| region                           | SiH <sub>4</sub>                                                                  | 50                          |                                            |                       | 20                   |
| 2nd layer                        | N <sub>2</sub>                                                                    | 500                         | 300                                        | 20                    | 0.4                  |
| region                           | PH <sub>3</sub> (against SiH <sub>4</sub> )                                       | 3000 ppm                    |                                            |                       | 5                    |
| 3rd layer                        | SiH <sub>4</sub>                                                                  | 40                          |                                            |                       |                      |
| region                           | CH <sub>4</sub>                                                                   | 600                         | 300                                        | 10                    | 0.4                  |
| 4th layer                        |                                                                                   |                             |                                            |                       | 0.3                  |
| region                           |                                                                                   |                             |                                            |                       |                      |

TABLE 203

| Order of lamination (layer name) | Gases and their flow rates (SCCM)                                                   | Substrate temperature (°C.) | RF discharging power (mW/cm³) | Inner pressure (Torr) | Layer thickness (μm) |
|----------------------------------|-------------------------------------------------------------------------------------|-----------------------------|-------------------------------|-----------------------|----------------------|
| Lower layer                      | SiH <sub>4</sub> 50                                                                 |                             |                               |                       |                      |
|                                  | B <sub>2</sub> H <sub>6</sub> (against SiH <sub>4</sub> ) 100 ppm                   |                             |                               |                       |                      |
|                                  | Cu(C <sub>4</sub> H <sub>7</sub> N <sub>2</sub> O <sub>2</sub> ) <sub>2</sub> /He 5 | 250                         | 5                             | 0.4                   | 0.05                 |
|                                  | GeF <sub>4</sub> 5                                                                  |                             |                               |                       |                      |
|                                  | H <sub>2</sub> 2 → 200*                                                             |                             |                               |                       |                      |
|                                  | AlCl <sub>3</sub> /He 200 → 20**                                                    |                             |                               |                       |                      |
| Upper layer                      | 1st layer region SiH <sub>4</sub> 100                                               |                             |                               |                       |                      |
|                                  | H <sub>2</sub> 300                                                                  | 250                         | 15                            | 0.4                   | 3                    |
|                                  | B <sub>2</sub> H <sub>6</sub> (against SiH <sub>4</sub> ) 250 ppm                   |                             |                               |                       |                      |
|                                  | AlCl <sub>3</sub> /He 1 → 0**                                                       |                             |                               |                       |                      |
|                                  | 2nd layer region SiH <sub>4</sub> 300                                               |                             |                               |                       |                      |
|                                  | H <sub>2</sub> 300                                                                  | 250                         | 15                            | 0.5                   | 10                   |
| 3rd layer region                 | SiH <sub>4</sub> 200                                                                |                             |                               |                       |                      |
|                                  | C <sub>2</sub> H <sub>2</sub> 10 → 20*                                              | 250                         | 15                            | 0.4                   | 20                   |
|                                  | NO 1                                                                                |                             |                               |                       |                      |

TABLE 204

| Order of lamination (layer name) | Gases and their flow rates (SCCM)                                                                  | Substrate temperature (°C.) | RF discharging power (mW/cm³) | Inner pressure (Torr) | Layer thickness (μm) |
|----------------------------------|----------------------------------------------------------------------------------------------------|-----------------------------|-------------------------------|-----------------------|----------------------|
| Lower layer                      | SiH <sub>4</sub> 50                                                                                |                             |                               |                       |                      |
|                                  | PH <sub>3</sub> (against SiH <sub>4</sub> ) 100 ppm                                                |                             |                               |                       |                      |
|                                  | Cu(C <sub>4</sub> H <sub>7</sub> N <sub>2</sub> O <sub>2</sub> ) <sub>2</sub> /He 5                |                             |                               |                       |                      |
|                                  | Mg(C <sub>5</sub> H <sub>5</sub> ) <sub>2</sub> /He 10                                             |                             |                               |                       |                      |
|                                  | H <sub>2</sub> 5 → 200*                                                                            | 250                         | 1                             | 0.4                   | 0.02                 |
|                                  | AlCl <sub>3</sub> /He (S-side: 0.01 μm) 200 → 30**<br>(UL-side: 0.01 μm)                           |                             |                               |                       |                      |
| Upper layer                      | SiH <sub>4</sub> 100                                                                               |                             |                               |                       |                      |
|                                  | H <sub>2</sub> 300                                                                                 |                             |                               |                       |                      |
|                                  | PH <sub>3</sub> (against SiH <sub>4</sub> ) 250 ppm<br>(LL-side: 2 μm)<br>(U · 2nd · LR-side 1 μm) | 250                         | 10                            | 0.4                   | 3                    |
|                                  | SiF <sub>4</sub> 5                                                                                 |                             |                               |                       |                      |
|                                  | SiH <sub>4</sub> 300                                                                               |                             |                               |                       |                      |
|                                  | H <sub>2</sub> 300                                                                                 | 300                         | 20                            | 0.5                   | 5                    |
| 2nd layer region                 | SiF <sub>4</sub> 20                                                                                |                             |                               |                       |                      |
|                                  | SiH <sub>4</sub> 100                                                                               |                             |                               |                       |                      |
|                                  | CH <sub>4</sub> 100                                                                                | 300                         | 15                            | 0.4                   | 20                   |
|                                  | SiF <sub>4</sub> 5                                                                                 |                             |                               |                       |                      |
|                                  | SiH <sub>4</sub> 50                                                                                |                             |                               |                       |                      |
|                                  | CH <sub>4</sub> 600                                                                                | 300                         | 10                            | 0.4                   | 0.5                  |
| 3rd layer region                 | SiF <sub>4</sub> 5                                                                                 |                             |                               |                       |                      |
|                                  |                                                                                                    |                             |                               |                       |                      |
| 4th layer region                 |                                                                                                    |                             |                               |                       |                      |
|                                  |                                                                                                    |                             |                               |                       |                      |
| 5th layer region                 |                                                                                                    |                             |                               |                       |                      |
|                                  |                                                                                                    |                             |                               |                       |                      |

TABLE 205

| Order of lamination (layer name) | Gases and their flow rates (SCCM)                                                         | Substrate temperature (°C.) | RF discharging power (mW/cm³) | Inner pressure (Torr) | Layer thickness (μm) |
|----------------------------------|-------------------------------------------------------------------------------------------|-----------------------------|-------------------------------|-----------------------|----------------------|
| Lower layer                      | SiH <sub>4</sub> 10 → 100*                                                                |                             |                               |                       |                      |
|                                  | Cu(C <sub>4</sub> H <sub>7</sub> N <sub>2</sub> O <sub>2</sub> ) <sub>2</sub> /He 1 → 10* |                             |                               |                       |                      |
|                                  | H <sub>2</sub> 5 → 200*                                                                   | 300                         | 5                             | 0.4                   | 0.2                  |
|                                  | AlCl <sub>3</sub> /He (S-side: 0.05 μm) 200 → 40**<br>(UL-side: 0.15 μm)                  |                             |                               |                       |                      |
|                                  | 40 → 10**                                                                                 |                             |                               |                       |                      |
|                                  |                                                                                           |                             |                               |                       |                      |
| Upper layer                      | SiH <sub>4</sub> 100                                                                      |                             |                               |                       |                      |
|                                  | H <sub>2</sub> 500                                                                        | 300                         | 10                            | 0.4                   | 3                    |
|                                  | B <sub>2</sub> H <sub>6</sub> (against SiH <sub>4</sub> ) 200 ppm                         |                             |                               |                       |                      |
|                                  | SiH <sub>4</sub> 100                                                                      |                             |                               |                       |                      |
|                                  | H <sub>2</sub> 300                                                                        | 300                         | 5                             | 0.2                   | 8                    |
|                                  |                                                                                           |                             |                               |                       |                      |
| 3rd layer region                 | SiH <sub>4</sub> 300                                                                      |                             |                               |                       |                      |
|                                  | NH <sub>3</sub> 50                                                                        | 300                         | 15                            | 0.4                   | 25                   |
| 4th layer region                 | SiH <sub>4</sub> 100                                                                      |                             |                               |                       |                      |
|                                  | NH <sub>3</sub> 50                                                                        | 300                         | 10                            | 0.4                   | 0.3                  |

TABLE 205-continued

| Order of lamination<br>(layer name) | Gases and<br>their flow rates<br>(SCCM) | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|-----------------------------------------|-----------------------------------|--------------------------------------------------|-----------------------------|----------------------------|
| region                              |                                         |                                   |                                                  |                             |                            |

TABLE 206

| Order of lamination<br>(layer name) | Gases and<br>their flow rates<br>(SCCM)                                                                                                                                                                                                                                   | Substrate<br>temperature<br>(°C.)                                                               | RF discharging<br>power<br>(mW/cm <sup>3</sup> ) | Inner<br>pressure<br>(Torr) | Layer<br>thickness<br>(μm) |
|-------------------------------------|---------------------------------------------------------------------------------------------------------------------------------------------------------------------------------------------------------------------------------------------------------------------------|-------------------------------------------------------------------------------------------------|--------------------------------------------------|-----------------------------|----------------------------|
| Lower layer                         | SiH <sub>4</sub><br>Cu(C <sub>4</sub> H <sub>7</sub> N <sub>2</sub> O <sub>2</sub> ) <sub>2</sub> /He<br>B <sub>2</sub> H <sub>6</sub> (against SiH <sub>4</sub> )<br>CH <sub>4</sub><br>GeH <sub>4</sub><br>H <sub>2</sub><br>AlCl <sub>3</sub> /He<br>(S-side: 0.05 μm) | 10 → 100*<br>5<br>10 ppm<br>2 → 20*<br>1 → 10*<br>5 → 200*<br>200 → 40**<br>(UL-side: 0.15 μm)  | 250                                              | 5                           | 0.4<br>0.2                 |
| Upper layer                         | 1st<br>layer<br>region                                                                                                                                                                                                                                                    | SiH <sub>4</sub><br>H <sub>2</sub><br>B <sub>2</sub> H <sub>6</sub> (against SiH <sub>4</sub> ) | 100<br>300<br>200 ppm                            | 250                         | 10<br>0.4<br>3             |
|                                     | 2nd<br>layer<br>region                                                                                                                                                                                                                                                    | SiH <sub>4</sub><br>SiF <sub>4</sub>                                                            | 100<br>5                                         | 300                         | 0.5<br>3                   |
|                                     | 3rd<br>layer<br>region                                                                                                                                                                                                                                                    | SiH <sub>4</sub><br>CH <sub>4</sub><br>PH <sub>3</sub> (against SiH <sub>4</sub> )              | 100<br>100<br>50 ppm                             | 300                         | 15<br>0.4<br>30            |
|                                     | 4th<br>layer<br>region                                                                                                                                                                                                                                                    | SiH <sub>4</sub><br>CH <sub>4</sub><br>SiF <sub>4</sub>                                         | 50<br>600<br>5                                   | 300                         | 10<br>0.4<br>0.5           |

TABLE 207

| Order of lamination<br>(layer name) | Gases and<br>their flow rates<br>(SCCM)                                                                                                                                               | Substrate<br>temperature<br>(°C.)                                                                                            | RF discharging<br>power<br>(mW/cm <sup>3</sup> )           | Inner<br>pressure<br>(Torr) | Layer<br>thickness<br>(μm) |
|-------------------------------------|---------------------------------------------------------------------------------------------------------------------------------------------------------------------------------------|------------------------------------------------------------------------------------------------------------------------------|------------------------------------------------------------|-----------------------------|----------------------------|
| Lower layer                         | SiH <sub>4</sub><br>PH <sub>3</sub> (against SiH <sub>4</sub> )<br>C <sub>2</sub> H <sub>2</sub><br>Cu(C <sub>4</sub> H <sub>7</sub> N <sub>2</sub> O <sub>2</sub> ) <sub>2</sub> /He | 50<br>10 ppm<br>5<br>250                                                                                                     | 5                                                          | 0.4                         | 0.05                       |
| Upper layer                         | 1st<br>layer<br>region                                                                                                                                                                | H <sub>2</sub><br>AlCl <sub>3</sub> /He<br>SiH <sub>4</sub><br>H <sub>2</sub><br>PH <sub>3</sub> (against SiH <sub>4</sub> ) | 3 → 1**<br>5 → 200*<br>200 → 20**<br>100<br>300<br>100 ppm | 250                         | 10<br>0.4<br>3             |
|                                     | 2nd<br>layer<br>region                                                                                                                                                                | Si <sub>2</sub> H <sub>6</sub><br>H <sub>2</sub><br>Si <sub>2</sub> F <sub>6</sub>                                           | 200<br>200<br>10                                           | 300                         | 10<br>0.5<br>10            |
|                                     | 3rd<br>layer<br>region                                                                                                                                                                | SiH <sub>4</sub><br>C <sub>2</sub> H <sub>2</sub>                                                                            | 300<br>50                                                  | 330                         | 20<br>0.4<br>30            |
|                                     | 4th<br>layer<br>region                                                                                                                                                                | B <sub>2</sub> H <sub>6</sub> (against SiH <sub>4</sub> )<br>(U · 2nd · LR-side: 1 μm)<br>(U · 4th · LR-side: 28 μm)         | 0 → 100 ppm*<br>100 ppm                                    | 20<br>0.4<br>1              |                            |

TABLE 208

| Order of lamination<br>(layer name) | Gases and<br>their flow rates<br>(SCCM)                                                                             | Substrate<br>temperature<br>(°C.) | RF discharging<br>power<br>(mW/cm <sup>3</sup> ) | Inner<br>pressure<br>(Torr) | Layer<br>thickness<br>(μm) |
|-------------------------------------|---------------------------------------------------------------------------------------------------------------------|-----------------------------------|--------------------------------------------------|-----------------------------|----------------------------|
| Lower layer                         | Si <sub>2</sub> F <sub>6</sub><br>Cu(C <sub>4</sub> H <sub>7</sub> N <sub>2</sub> O <sub>2</sub> ) <sub>2</sub> /He | 1<br>1 → 5*                       |                                                  |                             |                            |
|                                     | NO                                                                                                                  | 1 → 10*                           |                                                  |                             |                            |
|                                     | SiH <sub>4</sub>                                                                                                    | 10 → 100*                         | 250                                              | 5                           | 0.4<br>0.2                 |
|                                     | H <sub>2</sub>                                                                                                      | 5 → 200*                          |                                                  |                             |                            |
|                                     | AlCl <sub>3</sub> /He<br>(S-side: 0.05 μm)                                                                          |                                   |                                                  |                             |                            |

TABLE 208-continued

| Order of lamination (layer name) | Gases and their flow rates (SCCM)                         |                                             | Substrate temperature (°C.) | RF discharging power (mW/cm <sup>3</sup> ) | Inner pressure (Torr) | Layer thickness (μm) |    |
|----------------------------------|-----------------------------------------------------------|---------------------------------------------|-----------------------------|--------------------------------------------|-----------------------|----------------------|----|
| Upper layer                      | (UL-side: 0.15 μm)                                        |                                             | 200 → 40**                  |                                            |                       |                      |    |
|                                  | SiH <sub>4</sub>                                          |                                             | 40 → 10**                   |                                            |                       |                      |    |
|                                  | SiH <sub>4</sub>                                          | 100                                         |                             |                                            |                       |                      |    |
|                                  | H <sub>2</sub>                                            | 500                                         | 250                         | 10                                         | 0.4                   | 3                    |    |
|                                  | B <sub>2</sub> H <sub>6</sub> (against SiH <sub>4</sub> ) | 200 ppm                                     |                             |                                            |                       |                      |    |
|                                  | Si <sub>2</sub> F <sub>6</sub>                            | 10                                          |                             |                                            |                       |                      |    |
|                                  | SiH <sub>4</sub>                                          | 100                                         |                             |                                            |                       |                      |    |
|                                  | H <sub>2</sub>                                            | 300                                         | 300                         | 5                                          | 0.2                   | 8                    |    |
|                                  | Si <sub>2</sub> F <sub>6</sub>                            | 10                                          |                             |                                            |                       |                      |    |
|                                  | SiH <sub>4</sub>                                          | 300                                         |                             |                                            |                       |                      |    |
| Lower layer                      | 3rd layer                                                 | NH <sub>3</sub>                             | 30 → 50*                    | 300                                        | 15                    | 0.4                  | 25 |
|                                  | region                                                    | PH <sub>3</sub> (against SiH <sub>4</sub> ) | 50 ppm                      |                                            |                       |                      |    |
|                                  | SiH <sub>4</sub>                                          | 30                                          |                             |                                            |                       |                      |    |
|                                  | 4th layer                                                 | Si <sub>2</sub> F <sub>6</sub>              | 30                          |                                            |                       |                      |    |
|                                  | region                                                    | SiH <sub>4</sub>                            | 100                         |                                            |                       |                      |    |
|                                  | NH <sub>3</sub>                                           | 80 → 100*                                   | 300                         | 5                                          | 0.4                   | 0.7                  |    |
|                                  | region                                                    | PH <sub>3</sub> (against SiH <sub>4</sub> ) | 500 ppm                     |                                            |                       |                      |    |
|                                  | Si <sub>2</sub> F <sub>6</sub>                            | 10                                          |                             |                                            |                       |                      |    |

TABLE 209

| Order of lamination (layer name) | Gases and their flow rates (SCCM)                                                 |                                                           | Substrate temperature (°C.) | RF discharging power (mW/cm <sup>3</sup> ) | Inner pressure (Torr) | Layer thickness (μm) |   |
|----------------------------------|-----------------------------------------------------------------------------------|-----------------------------------------------------------|-----------------------------|--------------------------------------------|-----------------------|----------------------|---|
| Upper layer                      | (UL-side: 0.01 μm)                                                                |                                                           |                             |                                            |                       |                      |   |
|                                  | Cu(C <sub>4</sub> H <sub>7</sub> N <sub>2</sub> O <sub>2</sub> ) <sub>2</sub> /He | 20                                                        |                             |                                            |                       |                      |   |
|                                  | B <sub>2</sub> H <sub>6</sub> (against SiH <sub>4</sub> )                         | 100 ppm                                                   |                             |                                            |                       |                      |   |
|                                  | SiH <sub>4</sub>                                                                  | 50                                                        |                             |                                            |                       |                      |   |
|                                  | H <sub>2</sub>                                                                    | 5 → 200*                                                  | 250                         | 1                                          | 0.4                   | 0.02                 |   |
|                                  | AlCl <sub>3</sub> /He (S-side: 0.01 μm)                                           | 200 → 30**                                                |                             |                                            |                       |                      |   |
|                                  | SiH <sub>4</sub>                                                                  | 30 → 10**                                                 |                             |                                            |                       |                      |   |
|                                  | H <sub>2</sub>                                                                    | 100                                                       |                             |                                            |                       |                      |   |
|                                  | region                                                                            | B <sub>2</sub> H <sub>6</sub> (against SiH <sub>4</sub> ) | 200 ppm                     |                                            |                       |                      |   |
|                                  | 2nd layer                                                                         | SiH <sub>4</sub>                                          | 300                         |                                            |                       |                      |   |
| Lower layer                      | layer                                                                             | H <sub>2</sub>                                            | 500                         | 20                                         | 0.5                   | 20                   |   |
|                                  | region                                                                            | SiH <sub>4</sub>                                          | 100                         |                                            |                       |                      |   |
|                                  | 3rd layer                                                                         | GeH <sub>3</sub>                                          | 10 → 50*                    | 300                                        | 5                     | 0.4                  | 1 |
|                                  | region                                                                            | H <sub>2</sub>                                            | 300                         |                                            |                       |                      |   |
|                                  | 4th layer                                                                         | SiH <sub>4</sub>                                          | 100 → 40**                  | 300                                        | 10                    | 0.4                  | 1 |
|                                  | region                                                                            | CH <sub>4</sub>                                           | 100 → 600*                  |                                            |                       |                      |   |
|                                  | SiH <sub>4</sub>                                                                  | 200 → 30**                                                |                             |                                            |                       |                      |   |
|                                  | H <sub>2</sub>                                                                    | 30 → 10**                                                 |                             |                                            |                       |                      |   |
|                                  | region                                                                            | B <sub>2</sub> H <sub>6</sub> (against SiH <sub>4</sub> ) | 200 ppm                     |                                            |                       |                      |   |

TABLE 210

| Order of lamination (layer name) | Gases and their flow rates (SCCM)                                                 |                                                           | Substrate temperature (°C.) | RF discharging power (mW/cm <sup>3</sup> ) | Inner pressure (Torr) | Layer thickness (μm) |
|----------------------------------|-----------------------------------------------------------------------------------|-----------------------------------------------------------|-----------------------------|--------------------------------------------|-----------------------|----------------------|
| Upper layer                      | (UL-side: 0.01 μm)                                                                |                                                           |                             |                                            |                       |                      |
|                                  | B <sub>2</sub> H <sub>6</sub> (against SiH <sub>4</sub> )                         | 50 ppm                                                    |                             |                                            |                       |                      |
|                                  | NO                                                                                | 5                                                         |                             |                                            |                       |                      |
|                                  | Cu(C <sub>4</sub> H <sub>7</sub> N <sub>2</sub> O <sub>2</sub> ) <sub>2</sub> /He | 25                                                        |                             |                                            |                       |                      |
|                                  | SiH <sub>4</sub>                                                                  | 50                                                        |                             |                                            |                       |                      |
|                                  | H <sub>2</sub>                                                                    | 5 → 200*                                                  | 300                         | 1                                          | 0.3                   | 0.02                 |
|                                  | AlCl <sub>3</sub> /He (S-side: 0.01 μm)                                           | 200 → 30**                                                |                             |                                            |                       |                      |
|                                  | SiH <sub>4</sub>                                                                  | 30 → 10**                                                 |                             |                                            |                       |                      |
|                                  | H <sub>2</sub>                                                                    | 100                                                       |                             |                                            |                       |                      |
|                                  | region                                                                            | B <sub>2</sub> H <sub>6</sub> (against SiH <sub>4</sub> ) | 180 ppm                     |                                            |                       |                      |
| Lower layer                      | 1st layer                                                                         | (LL-side: 2.5 μm)                                         |                             |                                            |                       |                      |
|                                  | region                                                                            | (U · 2nd · LR-side: 0.5 μm)                               |                             |                                            |                       |                      |
|                                  | 2nd layer                                                                         | SiH <sub>4</sub>                                          | 180 → 0 ppm**               |                                            |                       |                      |
|                                  | region                                                                            | H <sub>2</sub>                                            | 300                         | 15                                         | 0.5                   | 20                   |
|                                  | 3rd layer                                                                         | SiH <sub>4</sub>                                          | 400                         | 300                                        | 10                    | 0.4                  |
| SiH <sub>4</sub>                 | region                                                                            | CH <sub>4</sub>                                           | 50                          |                                            |                       |                      |
|                                  | SiH <sub>4</sub>                                                                  | 500                                                       |                             |                                            |                       |                      |

TABLE 211

| Order of lamination (layer name) | Gases and their flow rates (SCCM)                                                                                                                                                                                                                                                                        | Substrate temperature (°C.)                                                                                                        | RF discharging power (mW/cm <sup>3</sup> ) | Inner pressure (Torr) | Layer thickness (μm) |     |
|----------------------------------|----------------------------------------------------------------------------------------------------------------------------------------------------------------------------------------------------------------------------------------------------------------------------------------------------------|------------------------------------------------------------------------------------------------------------------------------------|--------------------------------------------|-----------------------|----------------------|-----|
| Lower layer                      | SiH <sub>4</sub> 50<br>Cu(C <sub>4</sub> H <sub>7</sub> N <sub>2</sub> O <sub>2</sub> ) <sub>2</sub> /He 20<br>B <sub>2</sub> H <sub>6</sub> (against SiH <sub>4</sub> ) 50 ppm<br>NO 4<br>H <sub>2</sub> 5 → 200*<br>AlCl <sub>3</sub> /He (S-side: 0.01 μm) 200 → 30**<br>(UL-side: 0.01 μm) 30 → 10** | 300                                                                                                                                | 0.7                                        | 0.3                   | 0.02                 |     |
| Upper layer                      | 1st layer region                                                                                                                                                                                                                                                                                         | SiH <sub>4</sub> 80<br>H <sub>2</sub> 400<br>B <sub>2</sub> H <sub>6</sub> (against SiH <sub>4</sub> ) 200 ppm<br>2nd layer region | 300                                        | 7                     | 0.3                  | 3   |
|                                  | 3rd layer region                                                                                                                                                                                                                                                                                         | SiH <sub>4</sub> 200<br>H <sub>2</sub> 400                                                                                         | 300                                        | 12                    | 0.4                  | 20  |
|                                  |                                                                                                                                                                                                                                                                                                          | SiH <sub>4</sub> 40<br>CH <sub>4</sub> 400                                                                                         | 300                                        | 7                     | 0.3                  | 0.5 |

TABLE 212

| Order of lamination (layer name) | Gases and their flow rates (SCCM)                                                                                                                                                                                                                                                                       | Substrate temperature (°C.)                                                                                                        | RF discharging power (mW/cm <sup>3</sup> ) | Inner pressure (Torr) | Layer thickness (μm) |     |
|----------------------------------|---------------------------------------------------------------------------------------------------------------------------------------------------------------------------------------------------------------------------------------------------------------------------------------------------------|------------------------------------------------------------------------------------------------------------------------------------|--------------------------------------------|-----------------------|----------------------|-----|
| Lower layer                      | Cu(C <sub>4</sub> H <sub>7</sub> N <sub>2</sub> O <sub>2</sub> ) <sub>2</sub> /He 15<br>B <sub>2</sub> H <sub>6</sub> (against SiH <sub>4</sub> ) 50 ppm<br>NO 3<br>SiH <sub>4</sub> 25<br>H <sub>2</sub> 5 → 100*<br>AlCl <sub>3</sub> /He (S-side: 0.01 μm) 100 → 15**<br>(UL-side: 0.01 μm) 15 → 5** | 300                                                                                                                                | 0.5                                        | 0.2                   | 0.02                 |     |
| Upper layer                      | 1st layer region                                                                                                                                                                                                                                                                                        | SiH <sub>4</sub> 60<br>H <sub>2</sub> 280<br>B <sub>2</sub> H <sub>6</sub> (against SiH <sub>4</sub> ) 200 ppm<br>2nd layer region | 300                                        | 5                     | 0.3                  | 3   |
|                                  | 3rd layer region                                                                                                                                                                                                                                                                                        | SiH <sub>4</sub> 150<br>H <sub>2</sub> 300                                                                                         | 300                                        | 10                    | 0.4                  | 20  |
|                                  |                                                                                                                                                                                                                                                                                                         | SiH <sub>4</sub> 30<br>CH <sub>4</sub> 300                                                                                         | 300                                        | 5                     | 0.3                  | 0.5 |

TABLE 213

| Order of lamination (layer name) | Gases and their flow rates (SCCM)                                                                                                                                                                                                                                                                      | Substrate temperature (°C.)                                                                                                        | RF discharging power (mW/cm <sup>3</sup> ) | Inner pressure (Torr) | Layer thickness (μm) |     |
|----------------------------------|--------------------------------------------------------------------------------------------------------------------------------------------------------------------------------------------------------------------------------------------------------------------------------------------------------|------------------------------------------------------------------------------------------------------------------------------------|--------------------------------------------|-----------------------|----------------------|-----|
| Lower layer                      | Cu(C <sub>4</sub> H <sub>7</sub> N <sub>2</sub> O <sub>2</sub> ) <sub>2</sub> /He 10<br>B <sub>2</sub> H <sub>6</sub> (against SiH <sub>4</sub> ) 50 ppm<br>NO 2<br>SiH <sub>4</sub> 20<br>H <sub>2</sub> 5 → 100*<br>AlCl <sub>3</sub> /He (S-side: 0.01 μm) 80 → 15**<br>(UL-side: 0.01 μm) 15 → 5** | 300                                                                                                                                | 0.3                                        | 0.2                   | 0.02                 |     |
| Upper layer                      | 1st layer region                                                                                                                                                                                                                                                                                       | SiH <sub>4</sub> 40<br>H <sub>2</sub> 280<br>B <sub>2</sub> H <sub>6</sub> (against SiH <sub>4</sub> ) 200 ppm<br>2nd layer region | 300                                        | 3                     | 0.2                  | 3   |
|                                  | 3rd layer region                                                                                                                                                                                                                                                                                       | SiH <sub>4</sub> 100<br>H <sub>2</sub> 300                                                                                         | 300                                        | 6                     | 0.3                  | 20  |
|                                  |                                                                                                                                                                                                                                                                                                        | SiH <sub>4</sub> 20<br>CH <sub>4</sub> 200                                                                                         | 300                                        | 3                     | 0.2                  | 0.5 |

TABLE 213

| Order of lamination<br>(layer name) | Gases and their flow rates<br>(SCCM)                                              | Substrate temperature<br>(°C.)                            | RF discharging power<br>(mW/cm <sup>3</sup> ) | Inner pressure<br>(Torr) | Layer thickness<br>(μm) |
|-------------------------------------|-----------------------------------------------------------------------------------|-----------------------------------------------------------|-----------------------------------------------|--------------------------|-------------------------|
| Lower layer                         | SiH <sub>4</sub>                                                                  | 50                                                        |                                               |                          |                         |
|                                     | C <sub>2</sub> H <sub>2</sub>                                                     | 5                                                         |                                               |                          |                         |
|                                     | B <sub>2</sub> H <sub>6</sub> (against SiH <sub>4</sub> )                         | 10 ppm                                                    | 500                                           | 5                        | 0.4                     |
|                                     | Cu(C <sub>4</sub> H <sub>7</sub> N <sub>2</sub> O <sub>2</sub> ) <sub>2</sub> /He | 20                                                        |                                               |                          |                         |
|                                     | H <sub>2</sub>                                                                    | 5 → 200*                                                  |                                               |                          |                         |
| Upper layer                         | AlCl <sub>3</sub> /He                                                             | 200 → 20**                                                |                                               |                          |                         |
|                                     | 1st layer                                                                         | SiH <sub>4</sub>                                          | 100                                           |                          |                         |
|                                     | 2nd layer                                                                         | H <sub>2</sub>                                            | 1200                                          | 30                       | 0.4                     |
|                                     | region                                                                            | B <sub>2</sub> H <sub>6</sub> (against SiH <sub>4</sub> ) | 200 ppm                                       |                          |                         |
|                                     | 3rd layer                                                                         | SiH <sub>4</sub>                                          | 300                                           |                          |                         |
| region                              | H <sub>2</sub>                                                                    | 1500                                                      | 500                                           | 30                       | 0.5                     |
|                                     | SiH <sub>4</sub>                                                                  | 200                                                       |                                               |                          |                         |
|                                     | C <sub>2</sub> H <sub>2</sub>                                                     | 10 → 20*                                                  | 500                                           | 30                       | 0.4                     |
| region                              | NO                                                                                | 1                                                         |                                               |                          | 20                      |

TABLE 215

| Order of lamination<br>(layer name) | Gases and their flow rates<br>(SCCM)                                              | Substrate temperature<br>(°C.) | μW discharging power<br>(mW/cm <sup>3</sup> ) | Inner pressure<br>(Torr) | Layer thickness<br>(μm) |
|-------------------------------------|-----------------------------------------------------------------------------------|--------------------------------|-----------------------------------------------|--------------------------|-------------------------|
| Lower layer                         | SiF <sub>4</sub>                                                                  | 10                             |                                               |                          |                         |
|                                     | Cu(C <sub>4</sub> H <sub>7</sub> N <sub>2</sub> O <sub>2</sub> ) <sub>2</sub> /He | 10                             |                                               |                          |                         |
|                                     | B <sub>2</sub> H <sub>6</sub> (against SiH <sub>4</sub> )                         | 100 ppm                        |                                               |                          |                         |
|                                     | NO                                                                                | 10                             |                                               |                          |                         |
|                                     | SiH <sub>4</sub>                                                                  | 150                            |                                               |                          |                         |
| Upper layer                         | H <sub>2</sub>                                                                    | 20 → 500*                      | 250                                           | 0.5                      | 0.6                     |
|                                     | AlCl <sub>3</sub> /He<br>(S-side: 0.01 μm)                                        | 400 → 80**                     |                                               |                          |                         |
|                                     | (UL-side: 0.01 μm)                                                                | 80 → 50**                      |                                               |                          |                         |
|                                     | GeH <sub>4</sub>                                                                  | 20                             |                                               |                          |                         |
|                                     | SiH <sub>4</sub>                                                                  | 500                            |                                               |                          |                         |
| 1st layer                           | H <sub>2</sub>                                                                    | 500                            | 250                                           | 0.5                      | 0.4                     |
|                                     | B <sub>2</sub> H <sub>6</sub> (against SiH <sub>4</sub> )                         | 200 ppm                        |                                               |                          |                         |
|                                     | SiF <sub>4</sub>                                                                  | 20                             |                                               |                          |                         |
|                                     | SiH <sub>4</sub>                                                                  | 700                            |                                               |                          |                         |
|                                     | SiF <sub>4</sub>                                                                  | 30                             | 250                                           | 0.5                      | 0.5                     |
| 2nd layer                           | H <sub>2</sub>                                                                    | 500                            |                                               |                          |                         |
|                                     | SiH <sub>4</sub>                                                                  | 150                            |                                               |                          |                         |
|                                     | CH <sub>4</sub>                                                                   | 500                            | 250                                           | 0.5                      | 1                       |
| 3rd layer                           |                                                                                   |                                |                                               |                          |                         |
| region                              |                                                                                   |                                |                                               |                          |                         |

TABLE 216

| Order of lamination<br>(layer name) | Gases and their flow rates<br>(SCCM)                                              | Substrate temperature<br>(°C.) | RF discharging power<br>(mW/cm <sup>3</sup> ) | Inner pressure<br>(Torr) | Layer thickness<br>(μm) |
|-------------------------------------|-----------------------------------------------------------------------------------|--------------------------------|-----------------------------------------------|--------------------------|-------------------------|
| Lower layer                         | GeF <sub>4</sub>                                                                  | 5                              |                                               |                          |                         |
|                                     | C <sub>2</sub> H <sub>2</sub>                                                     | 10                             |                                               |                          |                         |
|                                     | B <sub>2</sub> H <sub>6</sub> (against SiH <sub>4</sub> )                         | 100 ppm                        |                                               |                          |                         |
|                                     | Cu(C <sub>4</sub> H <sub>7</sub> N <sub>2</sub> O <sub>2</sub> ) <sub>2</sub> /He | 10                             | 250                                           | 5                        | 0.4                     |
|                                     | SiH <sub>4</sub>                                                                  | 50                             |                                               |                          |                         |
| Upper layer                         | H <sub>2</sub>                                                                    | 5 → 200*                       |                                               |                          |                         |
|                                     | AlCl <sub>3</sub> /He                                                             | 200 → 20**                     |                                               |                          |                         |
|                                     | SiH <sub>4</sub>                                                                  | 100                            |                                               |                          |                         |
|                                     | H <sub>2</sub>                                                                    | 200                            |                                               |                          |                         |
|                                     | B <sub>2</sub> H <sub>6</sub> (against SiH <sub>4</sub> )<br>(LL-side: 3 μm)      | 400 ppm                        | 250                                           | 15                       | 0.4                     |
| 1st layer                           | (U · 2nd · LR-side: 2 μm)                                                         | 400 → 0 ppm**                  |                                               |                          | 5                       |
|                                     | SiH <sub>4</sub>                                                                  | 200                            |                                               |                          |                         |
|                                     | C <sub>2</sub> H <sub>2</sub>                                                     | 10 → 20*                       | 250                                           | 15                       | 0.4                     |
| 2nd layer                           | NO                                                                                | 1                              |                                               |                          |                         |
|                                     | SiH <sub>4</sub>                                                                  | 300                            |                                               |                          |                         |
|                                     | H <sub>2</sub>                                                                    | 300                            | 250                                           | 15                       | 0.5                     |
| 3rd layer                           |                                                                                   |                                |                                               |                          |                         |
| region                              |                                                                                   |                                |                                               |                          |                         |

TABLE 217

| Order of lamination<br>(layer name) | Gases and their flow rates<br>(SCCM)                                                                                                                                                                                                                                                                                                                                                                       | Substrate temperature<br>(°C.) | RF discharging power<br>(mW/cm <sup>3</sup> ) | Inner pressure<br>(Torr) | Layer thickness<br>(μm) |
|-------------------------------------|------------------------------------------------------------------------------------------------------------------------------------------------------------------------------------------------------------------------------------------------------------------------------------------------------------------------------------------------------------------------------------------------------------|--------------------------------|-----------------------------------------------|--------------------------|-------------------------|
| Lower layer                         | CH <sub>4</sub> 10<br>PH <sub>3</sub> (against SiH <sub>4</sub> ) 100 ppm<br>SiF <sub>4</sub> 10<br>SiH <sub>4</sub> 50<br>H <sub>2</sub> 5 → 200*<br>AlCl <sub>3</sub> /He 250<br>(S-side: 0.01 μm) 200 → 30**<br>(UL-side: 0.01 μm) 30 → 10**<br>Cu(C <sub>4</sub> H <sub>7</sub> N <sub>2</sub> O <sub>2</sub> ) <sub>2</sub> /He 10                                                                    |                                | 1                                             | 0.4                      | 0.02                    |
| Upper layer                         | 1st layer region SiH <sub>4</sub> 100<br>H <sub>2</sub> 200<br>PH <sub>3</sub> (against SiH <sub>4</sub> ) 200 ppm<br>SiF <sub>4</sub> 10<br>2nd layer region SiH <sub>4</sub> 100<br>CH <sub>4</sub> 100<br>SiF <sub>4</sub> 10<br>3rd layer region SiH <sub>4</sub> 300<br>H <sub>2</sub> 300<br>SiF <sub>4</sub> 20<br>4th layer region SiH <sub>4</sub> 50<br>H <sub>2</sub> 600<br>SiF <sub>4</sub> 5 | 250                            | 10                                            | 0.4                      | 3                       |
|                                     |                                                                                                                                                                                                                                                                                                                                                                                                            | 300                            | 15                                            | 0.4                      | 20                      |
|                                     |                                                                                                                                                                                                                                                                                                                                                                                                            | 300                            | 20                                            | 0.5                      | 5                       |
|                                     |                                                                                                                                                                                                                                                                                                                                                                                                            | 300                            | 10                                            | 0.4                      | 0.5                     |

TABLE 218

| Order of lamination<br>(layer name) | Gases and their flow rates<br>(SCCM)                                                                                                                                                                                                                                                                                                                                          | Substrate temperature<br>(°C.) | RF discharging power<br>(mW/cm <sup>3</sup> ) | Inner pressure<br>(Torr) | Layer thickness<br>(μm) |
|-------------------------------------|-------------------------------------------------------------------------------------------------------------------------------------------------------------------------------------------------------------------------------------------------------------------------------------------------------------------------------------------------------------------------------|--------------------------------|-----------------------------------------------|--------------------------|-------------------------|
| Lower layer                         | SnH <sub>4</sub> 1 → 10*<br>NO 1 → 10*<br>SiH <sub>4</sub> 10 → 100*<br>Cu(C <sub>4</sub> H <sub>7</sub> N <sub>2</sub> O <sub>2</sub> ) <sub>2</sub> /He 5 → 10*<br>H <sub>2</sub> 5 → 200*<br>AlCl <sub>3</sub> /He 300<br>(S-side: 0.05 μm) 200 → 40**<br>(UL-side: 0.15 μm) 40 → 10**<br>Mg(C <sub>5</sub> H <sub>5</sub> ) <sub>2</sub> /He 3                            |                                | 5                                             | 0.4                      | 0.2                     |
| Upper layer                         | 1st layer region SiH <sub>4</sub> 100<br>H <sub>2</sub> 500<br>BF <sub>3</sub> (against SiH <sub>4</sub> ) 150 ppm<br>(LL-side: 2 μm)<br>(U · 2nd · LR-side: 1 μm) 150 → 0 ppm**<br>2nd layer region SiH <sub>4</sub> 300<br>NH <sub>3</sub> 50<br>3rd layer region SiH <sub>4</sub> 100<br>H <sub>2</sub> 300<br>4th layer region SiH <sub>4</sub> 100<br>NH <sub>3</sub> 50 | 300                            | 10                                            | 0.4                      | 3                       |
|                                     |                                                                                                                                                                                                                                                                                                                                                                               | 300                            | 15                                            | 0.4                      | 25                      |
|                                     |                                                                                                                                                                                                                                                                                                                                                                               | 300                            | 5                                             | 0.2                      | 8                       |
|                                     |                                                                                                                                                                                                                                                                                                                                                                               | 300                            | 10                                            | 0.4                      | 0.3                     |

TABLE 219

| Order of lamination<br>(layer name) | Gases and their flow rates<br>(SCCM)                                                                                                                                                                                                                                                                                                                                       | Substrate temperature<br>(°C.) | RF discharging power<br>(mW/cm <sup>3</sup> ) | Inner pressure<br>(Torr) | Layer thickness<br>(μm) |
|-------------------------------------|----------------------------------------------------------------------------------------------------------------------------------------------------------------------------------------------------------------------------------------------------------------------------------------------------------------------------------------------------------------------------|--------------------------------|-----------------------------------------------|--------------------------|-------------------------|
| Lower layer                         | PF <sub>3</sub> (against SiH <sub>4</sub> ) 10 ppm<br>Cu(C <sub>4</sub> H <sub>7</sub> N <sub>2</sub> O <sub>2</sub> ) <sub>2</sub> /He 1 → 10*<br>CH <sub>4</sub> 2 → 20*<br>SiH <sub>4</sub> 10 → 100*<br>H <sub>2</sub> 5 → 200*<br>AlCl <sub>3</sub> /He 250<br>(S-side: 0.05 μm) 200 → 40**<br>(UL-side: 0.15 μm) 40 → 10**                                           |                                | 5                                             | 0.4                      | 0.2                     |
| Upper layer                         | 1st layer region SiH <sub>4</sub> 100<br>H <sub>2</sub> 100<br>PF <sub>3</sub> (against SiH <sub>4</sub> ) 50 ppm<br>SiF <sub>4</sub> 10<br>2nd layer region SiH <sub>4</sub> 100<br>CH <sub>4</sub> 100<br>PF <sub>3</sub> (against SiH <sub>4</sub> ) 50 ppm<br>SiF <sub>4</sub> 10<br>3rd layer region SiH <sub>4</sub> 100<br>SiF <sub>4</sub> 5<br>H <sub>2</sub> 200 | 250                            | 10                                            | 0.4                      | 3                       |
|                                     |                                                                                                                                                                                                                                                                                                                                                                            | 300                            | 15                                            | 0.4                      | 30                      |
|                                     |                                                                                                                                                                                                                                                                                                                                                                            | 300                            | 3                                             | 0.5                      | 3                       |

TABLE 219-continued

| Order of lamination (layer name) | Gases and their flow rates (SCCM)                                | Substrate temperature (°C.) | RF discharging power (mW/cm <sup>3</sup> ) | Inner pressure (Torr) | Layer thickness (μm) |
|----------------------------------|------------------------------------------------------------------|-----------------------------|--------------------------------------------|-----------------------|----------------------|
| 4th layer region                 | SiH <sub>4</sub> 50<br>CH <sub>4</sub> 600<br>SiF <sub>4</sub> 5 | 300                         | 10                                         | 0.4                   | 0.5                  |

TABLE 220

| Order of lamination (layer name) | Gases and their flow rates (SCCM)                                                                                                                                                                                                                                                                              | Substrate temperature (°C.) | RF discharging power (mW/cm <sup>3</sup> ) | Inner pressure (Torr) | Layer thickness (μm) |
|----------------------------------|----------------------------------------------------------------------------------------------------------------------------------------------------------------------------------------------------------------------------------------------------------------------------------------------------------------|-----------------------------|--------------------------------------------|-----------------------|----------------------|
| Lower layer                      | GeH <sub>4</sub> 10<br>SiH <sub>4</sub> 50<br>Cu(C <sub>4</sub> H <sub>7</sub> N <sub>2</sub> O <sub>2</sub> ) <sub>2</sub> /He 10 → 3**<br>C <sub>2</sub> H <sub>2</sub> 5<br>H <sub>2</sub> 5 → 200*<br>AlCl <sub>3</sub> /He 200 → 20**<br>B <sub>2</sub> H <sub>6</sub> (against SiH <sub>4</sub> ) 10 ppm | 250                         | 5                                          | 0.4                   | 0.05                 |
| Upper layer                      | SiH <sub>4</sub> 100<br>H <sub>2</sub> 300<br>B <sub>2</sub> H <sub>6</sub> (against SiH <sub>4</sub> ) 200 ppm                                                                                                                                                                                                | 250                         | 10                                         | 0.4                   | 3                    |
| 1st layer region                 | SiH <sub>4</sub> 300<br>C <sub>2</sub> H <sub>2</sub> 50                                                                                                                                                                                                                                                       | 330                         | 20                                         | 0.4                   | 30                   |
| 2nd layer region                 | B <sub>2</sub> H <sub>6</sub> (against SiH <sub>4</sub> ) (U · 1st · LR-side: 1 μm) 0 → 100 ppm*<br>(U · 3rd · LR-side: 29 μm) 100 ppm                                                                                                                                                                         | 330                         | 10                                         | 0.5                   | 10                   |
| 3rd layer region                 | SiH <sub>6</sub> 200<br>H <sub>2</sub> 200                                                                                                                                                                                                                                                                     | 300                         | 10                                         | 0.5                   | 10                   |
| 4th layer region                 | SiH <sub>4</sub> 200<br>C <sub>2</sub> H <sub>2</sub> 200                                                                                                                                                                                                                                                      | 330                         | 10                                         | 0.4                   | 1                    |

TABLE 221

| Order of lamination (layer name) | Gases and their flow rates (SCCM)                                                                                                                                                                                                                                                   | Substrate temperature (°C.) | RF discharging power (mW/cm <sup>3</sup> ) | Inner pressure (Torr) | Layer thickness (μm) |
|----------------------------------|-------------------------------------------------------------------------------------------------------------------------------------------------------------------------------------------------------------------------------------------------------------------------------------|-----------------------------|--------------------------------------------|-----------------------|----------------------|
| Lower layer                      | SiH <sub>4</sub> 10 → 100*<br>NO 1 → 10*<br>GeF <sub>4</sub> 1 → 10*<br>H <sub>2</sub> 5 → 200*<br>AlCl <sub>3</sub> /He (S-side: 0.05 μm) 200 → 40**<br>(UL-side: 0.15 μm) 40 → 10**<br>Cu(C <sub>4</sub> H <sub>7</sub> N <sub>2</sub> O <sub>2</sub> ) <sub>2</sub> /He 20 → 5** | 250                         | 5                                          | 0.4                   | 0.2                  |
| Upper layer                      | SiH <sub>4</sub> 100<br>H <sub>2</sub> 100<br>PH <sub>3</sub> (against SiH <sub>4</sub> ) 150 ppm                                                                                                                                                                                   | 250                         | 10                                         | 0.4                   | 3                    |
| 1st layer region                 | SiH <sub>4</sub> 300<br>NH <sub>3</sub> 30 → 50*<br>PH <sub>3</sub> (against SiH <sub>4</sub> ) 50 ppm                                                                                                                                                                              | 300                         | 15                                         | 0.4                   | 25                   |
| 2nd layer region                 | SiH <sub>4</sub> 100<br>H <sub>2</sub> 300                                                                                                                                                                                                                                          | 300                         | 5                                          | 0.2                   | 8                    |
| 3rd layer region                 | SiH <sub>4</sub> 100<br>H <sub>2</sub> 300                                                                                                                                                                                                                                          | 300                         | 5                                          | 0.4                   | 0.7                  |
| 4th layer region                 | NH <sub>3</sub> 80 → 100*<br>B <sub>2</sub> H <sub>6</sub> (against SiH <sub>4</sub> ) 500 ppm                                                                                                                                                                                      | 300                         | 5                                          | 0.4                   | 0.7                  |

TABLE 222

| Order of lamination (layer name) | Gases and their flow rates (SCCM)                                                                                                                                                                                                                                                                | Substrate temperature (°C.) | RF discharging power (mW/cm <sup>3</sup> ) | Inner pressure (Torr) | Layer thickness (μm) |
|----------------------------------|--------------------------------------------------------------------------------------------------------------------------------------------------------------------------------------------------------------------------------------------------------------------------------------------------|-----------------------------|--------------------------------------------|-----------------------|----------------------|
| Lower layer                      | B <sub>2</sub> H <sub>6</sub> (against SiH <sub>4</sub> ) 50 ppm<br>Cu(C <sub>4</sub> H <sub>7</sub> N <sub>2</sub> O <sub>2</sub> ) <sub>2</sub> /He 10<br>SiH <sub>4</sub> 50<br>H <sub>2</sub> 5 → 200*<br>AlCl <sub>3</sub> /He (S-side: 0.01 μm) 200 → 30**<br>(UL-side: 0.01 μm) 30 → 10** | 250                         | 1                                          | 0.3                   | 0.02                 |
| Upper layer                      | SiH <sub>4</sub> 100<br>H <sub>2</sub> 300<br>B <sub>2</sub> H <sub>6</sub> (against SiH <sub>4</sub> ) 500 ppm                                                                                                                                                                                  | 250                         | 10                                         | 0.4                   | 3                    |
| 2nd layer                        | SiH <sub>4</sub> 300<br>H <sub>2</sub> 600                                                                                                                                                                                                                                                       | 250                         | 25                                         | 0.6                   | 25                   |

TABLE 222-continued

| Order of lamination<br>(layer name) | Gases and their flow rates<br>(SCCM) | Substrate temperature<br>(°C.) | RF discharging power<br>(mW/cm <sup>3</sup> ) | Inner pressure<br>(Torr) | Layer thickness<br>(μm) |
|-------------------------------------|--------------------------------------|--------------------------------|-----------------------------------------------|--------------------------|-------------------------|
| region                              |                                      |                                |                                               |                          |                         |
| 3rd layer                           | SiH <sub>4</sub> 50                  | 250                            | 10                                            | 0.4                      | 1                       |
| region                              | CH <sub>4</sub> 500                  |                                |                                               |                          |                         |

TABLE 223

| Order of lamination<br>(layer name) | Gases and their flow rates<br>(SCCM)                                                  | Substrate temperature<br>(°C.) | RF discharging power<br>(mW/cm <sup>3</sup> ) | Inner pressure<br>(Torr) | Layer thickness<br>(μm) |
|-------------------------------------|---------------------------------------------------------------------------------------|--------------------------------|-----------------------------------------------|--------------------------|-------------------------|
| Lower layer                         | SiH <sub>4</sub> 50                                                                   |                                |                                               |                          |                         |
|                                     | Cu(C <sub>4</sub> H <sub>7</sub> N <sub>2</sub> O <sub>2</sub> ) <sub>2</sub> /He 15  |                                |                                               |                          |                         |
|                                     | SiF <sub>4</sub> 1                                                                    |                                |                                               |                          |                         |
|                                     | B <sub>2</sub> H <sub>6</sub> (against SiH <sub>4</sub> ) 100 ppm                     |                                |                                               |                          |                         |
|                                     | H <sub>2</sub> 5 → 200*                                                               | 300                            | 2                                             | 0.3                      | 0.05                    |
|                                     | Al(CH <sub>3</sub> ) <sub>3</sub> /He                                                 |                                |                                               |                          |                         |
|                                     | (S-side: 0.03 μm) 200 → 50**                                                          |                                |                                               |                          |                         |
|                                     | (UL-side: 0.02 μm) 50 → 5**                                                           |                                |                                               |                          |                         |
| Upper layer                         | SiH <sub>4</sub> 100                                                                  |                                |                                               |                          |                         |
| 1st layer                           | H <sub>2</sub> 300                                                                    |                                |                                               |                          |                         |
| region                              | B <sub>2</sub> H <sub>6</sub> (against SiH <sub>4</sub> ) 700 ppm                     | 300                            | 10                                            | 0.4                      | 10                      |
|                                     | Al(CH <sub>3</sub> ) <sub>3</sub> /He 0.3                                             |                                |                                               |                          |                         |
|                                     | SiF <sub>4</sub> 5                                                                    |                                |                                               |                          |                         |
|                                     | Cu(C <sub>4</sub> H <sub>7</sub> N <sub>2</sub> O <sub>2</sub> ) <sub>2</sub> /He 0.3 |                                |                                               |                          |                         |
| 2nd layer                           | SiH <sub>4</sub> 300                                                                  |                                |                                               |                          |                         |
| region                              | H <sub>2</sub> 300                                                                    |                                |                                               |                          |                         |
|                                     | CH <sub>4</sub> 1                                                                     |                                |                                               |                          |                         |
|                                     | Al(CH <sub>3</sub> ) <sub>3</sub> /He 0.1                                             | 300                            | 25                                            | 0.5                      | 25                      |
|                                     | NO 0.1                                                                                |                                |                                               |                          |                         |
|                                     | SiF <sub>4</sub> 1                                                                    |                                |                                               |                          |                         |
|                                     | B <sub>2</sub> H <sub>6</sub> (against SiH <sub>4</sub> ) 0.5 ppm                     |                                |                                               |                          |                         |
|                                     | Cu(C <sub>4</sub> H <sub>7</sub> N <sub>2</sub> O <sub>2</sub> ) <sub>2</sub> /He 0.1 |                                |                                               |                          |                         |
| 3rd layer                           | SiH <sub>4</sub> 200                                                                  |                                |                                               |                          |                         |
| region                              | H <sub>2</sub> 200                                                                    |                                |                                               |                          |                         |
|                                     | B <sub>2</sub> H <sub>6</sub> (against SiH <sub>4</sub> ) 0.1 ppm                     |                                |                                               |                          |                         |
|                                     | PH <sub>3</sub> (against SiH <sub>4</sub> ) 1000 ppm                                  |                                |                                               |                          |                         |
|                                     | SiF <sub>4</sub> 1                                                                    |                                |                                               |                          |                         |
|                                     | NO 0.1                                                                                | 300                            | 15                                            | 0.4                      | 5                       |
|                                     | Al(CH <sub>3</sub> ) <sub>3</sub> /He 0.1                                             |                                |                                               |                          |                         |
|                                     | Cu(C <sub>4</sub> H <sub>7</sub> N <sub>2</sub> O <sub>2</sub> ) <sub>2</sub> /He 0.2 |                                |                                               |                          |                         |
|                                     | CH <sub>4</sub>                                                                       |                                |                                               |                          |                         |
|                                     | (U · 2nd · LR-side: 1 μm) 1 → 600*                                                    |                                |                                               |                          |                         |
|                                     | (U · 4th · LR-side: 4 μm) 600                                                         |                                |                                               |                          |                         |
| 4th layer                           | H <sub>2</sub> 200                                                                    |                                |                                               |                          |                         |
| region                              | SiF <sub>4</sub> 5                                                                    |                                |                                               |                          |                         |
|                                     | B <sub>2</sub> H <sub>6</sub> (against SiH <sub>4</sub> ) 1 ppm                       |                                |                                               |                          |                         |
|                                     | PH <sub>3</sub> (against SiH <sub>4</sub> ) 5 ppm                                     | 300                            | 10                                            | 0.4                      | 0.3                     |
|                                     | NO 0.5                                                                                |                                |                                               |                          |                         |
|                                     | CH <sub>4</sub> 600                                                                   |                                |                                               |                          |                         |
|                                     | Al(CH <sub>3</sub> ) <sub>3</sub> /He 0.5                                             |                                |                                               |                          |                         |
|                                     | Cu(C <sub>4</sub> H <sub>7</sub> N <sub>2</sub> O <sub>2</sub> ) <sub>2</sub> /He 0.1 |                                |                                               |                          |                         |
|                                     | SiH <sub>4</sub>                                                                      |                                |                                               |                          |                         |
|                                     | (U · 3rd · LR-side: 0.03 μm) 200 → 20**                                               |                                |                                               |                          |                         |
|                                     | (FS-side: 0.07 μM) 20                                                                 |                                |                                               |                          |                         |

TABLE 224

| Order of lamination<br>(layer name) | Gases and their flow rates<br>(SCCM)                              | Substrate temperature<br>(°C.) | RF discharging power<br>(mW/cm <sup>3</sup> ) | Inner pressure<br>(Torr) | Layer thickness<br>(μm) |
|-------------------------------------|-------------------------------------------------------------------|--------------------------------|-----------------------------------------------|--------------------------|-------------------------|
| Lower layer                         | SiH <sub>4</sub> 30                                               |                                |                                               |                          |                         |
|                                     | H <sub>2</sub> 5 → 100*                                           | 330                            | 1                                             | 0.01                     | 0.05                    |
|                                     | Ar 100                                                            |                                |                                               |                          |                         |
| Upper layer                         | SiH <sub>4</sub> 100                                              |                                |                                               |                          |                         |
| 1st layer                           | H <sub>2</sub> 300                                                | 330                            | 10                                            | 0.4                      | 3                       |
| region                              | B <sub>2</sub> H <sub>6</sub> (against SiH <sub>4</sub> ) 800 ppm |                                |                                               |                          |                         |
| 2nd layer                           | SiH <sub>4</sub> 400                                              |                                |                                               |                          |                         |
| region                              | H <sub>2</sub> 800                                                | 330                            | 25                                            | 0.5                      | 25                      |
| 3rd layer                           | SiH <sub>4</sub> 20                                               |                                |                                               |                          |                         |
| region                              | CH <sub>4</sub> 400                                               | 350                            | 10                                            | 0.4                      | 1                       |

TABLE 225

| Order of lamination (layer name) | Gases and their flow rates (SCCM)                         |            | Substrate temperature (°C.) | RF discharging power (mW/cm <sup>3</sup> ) | Inner pressure (Torr) | Layer thickness (μm) |
|----------------------------------|-----------------------------------------------------------|------------|-----------------------------|--------------------------------------------|-----------------------|----------------------|
| Lower layer                      | SiH <sub>4</sub>                                          | 5 → 50*    |                             |                                            |                       |                      |
|                                  | H <sub>2</sub>                                            | 10 → 200*  | 250                         | 5                                          | 0.4                   | 0.05                 |
|                                  | Al(CH <sub>3</sub> ) <sub>3</sub> /He                     | 120 → 40** |                             |                                            |                       |                      |
|                                  | NaNH <sub>2</sub> /He                                     | 10         |                             |                                            |                       |                      |
| Upper layer                      | SiH <sub>4</sub>                                          | 100        |                             |                                            |                       |                      |
|                                  | B <sub>2</sub> H <sub>6</sub> (against SiH <sub>4</sub> ) | 200 ppm    | 250                         | 10                                         | 0.4                   | 3                    |
|                                  | H <sub>2</sub>                                            | 100        |                             |                                            |                       |                      |
|                                  | SiH <sub>4</sub>                                          | 300        | 250                         | 15                                         | 0.5                   | 20                   |
| 1st layer region                 | H <sub>2</sub>                                            | 300        | 250                         | 15                                         | 0.5                   | 20                   |
|                                  | SiH <sub>4</sub>                                          | 50         | 250                         | 10                                         | 0.4                   | 0.5                  |
| 2nd layer region                 | SiH <sub>4</sub>                                          | 50         | 250                         | 10                                         | 0.4                   | 0.5                  |
|                                  | CH <sub>4</sub>                                           | 500        | 250                         | 10                                         | 0.4                   | 0.5                  |
| 3rd layer region                 | SiH <sub>4</sub>                                          | 50         | 250                         | 10                                         | 0.4                   | 0.5                  |
|                                  | CH <sub>4</sub>                                           | 500        | 250                         | 10                                         | 0.4                   | 0.5                  |

TABLE 226

|                                           | Comparative Example 2 | Example 1  | Example 2  |
|-------------------------------------------|-----------------------|------------|------------|
| Al(CH <sub>3</sub> ) <sub>3</sub> /He     |                       |            |            |
| Flow rates (sccm)                         | 120 → 10**            | 120 → 20** | 120 → 40** |
| Content of Al (atomic %)                  | 6                     | 12         | 20         |
| Ratio of film peeling-off (Example 1 = 1) | 25                    | 12         | 1          |
|                                           |                       | 26         | 37         |
|                                           |                       | 0.96       | 0.93       |

TABLE 227

| Order of lamination (layer name) | Gases and their flow rates (sccm)                   |         | 30 |
|----------------------------------|-----------------------------------------------------|---------|----|
| Lower layer                      | SiF <sub>4</sub>                                    | 3       |    |
|                                  | NO                                                  | 3       |    |
|                                  | CH <sub>4</sub>                                     | 2       |    |
|                                  | B <sub>2</sub> H <sub>2</sub>                       | 100 ppm | 35 |
| 1st layer region                 | SiF <sub>4</sub>                                    | 1       |    |
|                                  | Zn(C <sub>2</sub> H <sub>5</sub> ) <sub>2</sub> /He | 1       |    |
|                                  | SiF <sub>4</sub>                                    | 0.2     |    |
| Upper layer                      | NO                                                  | 0.1     |    |
|                                  | CH <sub>4</sub>                                     | 1       |    |
| 2nd layer region                 |                                                     |         |    |

TABLE 227-continued

| Order of lamination (layer name) | Gases and their flow rates (sccm)                         |         |
|----------------------------------|-----------------------------------------------------------|---------|
| 3rd layer region                 | Zn(C <sub>2</sub> H <sub>5</sub> ) <sub>2</sub> /He       | 0.3     |
|                                  | B <sub>2</sub> H <sub>6</sub> (against SiH <sub>4</sub> ) | 0.5 ppm |
|                                  | SiH <sub>4</sub>                                          | 1       |
|                                  | B <sub>2</sub> H <sub>6</sub> (against SiH <sub>4</sub> ) | 2 ppm   |
|                                  | NO                                                        | 0.5     |
|                                  | Al(CH <sub>3</sub> ) <sub>3</sub> /He                     | 0.5     |
|                                  | Zn(C <sub>2</sub> H <sub>5</sub> ) <sub>2</sub> /He       | 1       |

TABLE 228

| Order of lamination (layer name) | Gases and their flow rates (SCCM)                         |            | Substrate temperature (°C.) | RF discharging power (mW/cm <sup>3</sup> ) | Inner pressure (Torr) | Layer thickness (μm) |
|----------------------------------|-----------------------------------------------------------|------------|-----------------------------|--------------------------------------------|-----------------------|----------------------|
| Lower layer                      | SiH <sub>4</sub>                                          | 5 → 50*    |                             |                                            |                       |                      |
|                                  | H <sub>2</sub>                                            | 10 → 200*  |                             |                                            |                       |                      |
|                                  | Al(CH <sub>3</sub> ) <sub>3</sub> /He                     | 120 → 40** | 300                         | 5                                          | 0.4                   | 0.05                 |
|                                  | Y(oi-C <sub>3</sub> H <sub>7</sub> ) <sub>3</sub> /He     | 10         |                             |                                            |                       |                      |
| Upper layer                      | SiH <sub>4</sub>                                          | 100        |                             |                                            |                       |                      |
|                                  | B <sub>2</sub> H <sub>6</sub> (against SiH <sub>4</sub> ) | 200 ppm    | 250                         | 10                                         | 0.4                   | 5                    |
|                                  | H <sub>2</sub>                                            | 100        |                             |                                            |                       |                      |
|                                  | SiH <sub>4</sub>                                          | 200        |                             |                                            |                       |                      |
| 1st layer region                 | C <sub>2</sub> H <sub>2</sub>                             | 20         | 300                         | 30                                         | 0.5                   | 20                   |
|                                  | B <sub>2</sub> H <sub>6</sub> (against SiH <sub>4</sub> ) | 5 ppm      |                             |                                            |                       |                      |
|                                  | H <sub>2</sub>                                            | 500        |                             |                                            |                       |                      |
|                                  | SiH <sub>4</sub>                                          | 300        |                             |                                            |                       |                      |
| 2nd layer region                 | CH <sub>4</sub>                                           | 300        | 300                         | 15                                         | 0.5                   | 5                    |
|                                  | SiH <sub>4</sub>                                          | 50         |                             |                                            |                       |                      |
|                                  | CH <sub>4</sub>                                           | 500        | 300                         | 10                                         | 0.4                   | 0.5                  |
|                                  | SiH <sub>4</sub>                                          | 50         |                             |                                            |                       |                      |
| 3rd layer region                 | CH <sub>4</sub>                                           | 500        | 300                         |                                            |                       |                      |
|                                  | SiH <sub>4</sub>                                          | 50         |                             |                                            |                       |                      |
| 4th layer region                 | CH <sub>4</sub>                                           | 500        | 300                         |                                            |                       |                      |
|                                  | SiH <sub>4</sub>                                          | 50         |                             |                                            |                       |                      |
| 5th layer region                 | CH <sub>4</sub>                                           | 500        | 300                         |                                            |                       |                      |
|                                  | SiH <sub>4</sub>                                          | 50         |                             |                                            |                       |                      |

TABLE 229

| Order of lamination (layer name) | Gases and their flow rates (SCCM)     |            | Substrate temperature (°C.) | RF discharging power (mW/cm <sup>3</sup> ) | Inner pressure (Torr) | Layer thickness (μm) |
|----------------------------------|---------------------------------------|------------|-----------------------------|--------------------------------------------|-----------------------|----------------------|
| Lower layer                      | SiH <sub>4</sub>                      | 15 → 150*  |                             |                                            |                       |                      |
|                                  | SiF <sub>4</sub>                      | 10 → 20*   |                             |                                            |                       |                      |
|                                  | H <sub>2</sub>                        | 20 → 300*  | 250                         | 0.5                                        | 0.6                   | 0.07                 |
|                                  | Al(CH <sub>3</sub> ) <sub>3</sub> /He | 400 → 50** |                             |                                            |                       |                      |
|                                  | NaNH <sub>2</sub> /He                 | 20         |                             |                                            |                       |                      |

TABLE 229-continued

| Order of lamination (layer name) | Gases and their flow rates (SCCM) |                                                           | Substrate temperature (°C.) | RF discharging power (mW/cm <sup>3</sup> ) | Inner pressure (Torr) | Layer thickness (μm) |
|----------------------------------|-----------------------------------|-----------------------------------------------------------|-----------------------------|--------------------------------------------|-----------------------|----------------------|
| Upper layer                      | 1st layer region                  | SiH <sub>4</sub>                                          | 230                         | 250                                        | 0.5                   | 3                    |
|                                  |                                   | SiF <sub>4</sub>                                          | 20                          |                                            |                       |                      |
|                                  |                                   | B <sub>2</sub> H <sub>6</sub> (against SiH <sub>4</sub> ) | 150 ppm                     |                                            |                       |                      |
|                                  | 2nd layer region                  | H <sub>2</sub>                                            | 150                         | 250                                        | 0.5                   | 20                   |
|                                  |                                   | SiH <sub>4</sub>                                          | 700                         |                                            |                       |                      |
|                                  | 3rd layer region                  | SiF <sub>4</sub>                                          | 30                          |                                            |                       |                      |
|                                  |                                   | H <sub>2</sub>                                            | 500                         |                                            |                       |                      |
|                                  |                                   | SiH <sub>4</sub>                                          | 150                         |                                            |                       |                      |
|                                  |                                   | CH <sub>4</sub>                                           | 500                         | 250                                        | 0.5                   | 0.3                  |
|                                  |                                   |                                                           |                             |                                            |                       | 1                    |

TABLE 230

| Order of lamination (layer name) | Gases and their flow rates (SCCM) |          | Substrate temperature (°C.) | RF discharging power (mW/cm <sup>3</sup> ) | Inner pressure (Torr) | Layer thickness (μm) |
|----------------------------------|-----------------------------------|----------|-----------------------------|--------------------------------------------|-----------------------|----------------------|
| Lower layer                      | SiH <sub>4</sub>                  | 10 → 50* | 250                         | 1                                          | 0.01                  | 0.05                 |
|                                  | H <sub>2</sub>                    | 5 → 100* |                             |                                            |                       |                      |
|                                  | Ar                                | 200      |                             |                                            |                       |                      |

What is claimed is:

1. A light receiving member having an aluminum support and a multilayered light receiving layer exhibiting photoconductivity formed on said aluminum support, characterized in that said multilayered light receiving layer comprises: a lower layer (a) in contact with said support and an upper layer (b) having a free surface disposed on said lower layer (a); said lower layer (a) being formed of an inorganic material composed of aluminum atoms, silicon atoms, hydrogen atoms and atoms of an element capable of contributing to the control of image quality selected from the group consisting of boron, gallium, indium, thallium, phosphorus, arsenic, antimony, bismuth, sulfur, selenium, tellurium and polonium; said lower layer (a) having a portion in which said aluminum, silicon and hydrogen atoms are unevenly distributed across the layer thickness; said aluminum atoms being contained in said lower layer (a) such that their content decreases across the layer thickness upward from the interface between said lower layer (a) and said aluminum support and wherein said content of said aluminum atoms is lower than 95 atomic % in the vicinity of the interface between said lower layer (a) and said aluminum support and higher than 5 atomic % in the vicinity of the interface between said lower layer (a) and said upper layer (b); said upper layer (b) comprising a plurality of layer regions, each said region comprising a non-single-crystal material composed of silicon atoms as the matrix, and wherein the layer region adjacent said lower layer (a) comprises (i) a non-single-crystal material containing silicon atoms as the matrix, (ii) at least one kind of atoms selected from the group consisting of hydrogen atoms and halogen atoms, and (iii) atoms of a conductivity controlling element selected from the group consisting of Group III atoms, Group V atoms, except nitrogen, and Group VI atoms, except oxygen, of the periodic table.

2. A light receiving member according to claim 1, wherein the amount of said silicon atoms contained in the lower layer is from 5 to 95 atomic %.

3. A light receiving member according to claim 1, wherein the amount of said hydrogen atoms contained in the lower layer is from 0.01 to 70 atomic %.

4. A light receiving member according to claim 1, wherein the amount of said element atoms capable of contributing to the control of image quality contained

in the lower layer is from  $1 \times 10^{-3}$  to  $5 \times 10^4$  atomic ppm.

5. A light receiving member according to claim 1, wherein the lower layer further contains one kind of atoms selected from the group consisting of carbon atoms, nitrogen atoms and oxygen atoms.

6. A light receiving member according to claim 5, wherein the amount of said one kind of atoms contained in the lower layer is from  $1 \times 10^3$  to  $5 \times 10^5$  atomic ppm.

7. A light receiving member according to claim 1, wherein the lower layer further contains one kind of halogen atoms selected from the group consisting of fluorine atoms, chlorine atoms, bromine atoms and iodine atoms.

8. A light receiving member according to claim 7, wherein the amount of said one kind of halogen atoms contained in the lower layer is from  $1 \times 4 \times 10^5$  atomic ppm.

9. A light receiving member according to claim 5, wherein the lower layer further contains one kind of halogen atoms selected from the group consisting of fluorine atoms, chlorine atoms, bromine atoms and iodine atoms.

10. A light receiving member according to claim 9, wherein the amount of said one kind of halogen atoms contained in the lower layer is from 1 to  $4 \times 10^5$  atomic ppm.

11. A light receiving member according to claim 1, wherein the lower layer further contains one kind of atoms selected from the group consisting of germanium atoms and tin atoms.

12. A light receiving member according to claim 11, wherein the amount of said germanium or tin atoms contained in the lower layer is from 1 to  $9 \times 10^5$  atomic ppm.

13. A light receiving member according to claim 5, wherein the lower layer further contains one kind of atoms selected from the group consisting of germanium atoms and tin atoms.

14. A light receiving member according to claim 13, wherein the amount of said germanium or tin atoms contained in the lower layer is from 1 to  $9 \times 10^5$  atomic ppm.

15. A light receiving member according to claim 7, wherein the lower layer further contains one kind of

atoms selected from the group consisting of germanium atoms and tin atoms.

16. A light receiving member according to claim 15, wherein the amount of said germanium or tin atoms contained in the lower layer is from  $1 \times 10^5$  atomic ppm.

17. A light receiving member according to claim 1, wherein the lower layer further contains atoms of a metal selected from the group consisting of magnesium, copper, sodium, yttrium, manganese and zinc.

18. A light receiving member according to claim 17, wherein the amount of said metal atoms contained in the lower layer is from 1 to  $2 \times 10^5$  atomic ppm.

19. A light receiving member according to claim 5, wherein the lower layer further contains atoms of a metal selected from the group consisting of magnesium, copper, sodium, yttrium, manganese and zinc.

20. A light receiving member according to claim 19, wherein the amount of said metal atoms contained in the lower layer is from 1 to  $2 \times 10^5$  atomic ppm.

21. A light receiving member according to claim 7, wherein the lower layer further contains atoms of a metal selected from the group consisting of magnesium, copper, sodium, yttrium, manganese and zinc.

22. A light receiving member according to claim 21, wherein the amount of said metal atoms contained in the lower layer is from 1 to  $2 \times 10^5$  atomic ppm.

23. A light receiving member according to claim 11, wherein the lower layer further contains atoms of a metal selected from the group consisting of magnesium, copper, sodium, yttrium, manganese and zinc.

15

20

25

30

35

24. A light receiving member according to claim 23, wherein the amount of said metal atoms contained in the lower layer is from 1 to  $2 \times 10^5$  atomic ppm.

25. A light receiving member according to claim 1, wherein the amount of said atoms of a conductivity controlling element selected from Group III, Group V, except nitrogen, or Group VI, except oxygen, atoms of the periodic table contained in the lower region of the upper layer adjacent the lower layer is from  $1 \times 10^{-3}$  to  $5 \times 10^4$  atomic ppm.

26. A light receiving member according to claim 25, wherein said conductivity controlling element selected from Group III atoms of the periodic table is a member selected from the group consisting of boron, aluminum, gallium, indium and thallium.

27. A light receiving member according to claim 25, wherein said conductivity controlling element selected from Group V atoms of the periodic table is a member selected from the group consisting of phosphorous, arsenic, antimony and bismuth.

28. A light receiving member according to claim 25, wherein said conductivity controlling element selected from Group VI atoms of the periodic table is a member selected from the group consisting of sulfur, selenium, tellurium and polonium.

29. A light receiving member according to claim 1, wherein the lower layer is 0.03 to 5  $\mu\text{m}$  thick and the upper layer is 1 to 130  $\mu\text{m}$  thick.

30. An electrophotographic process comprising:  
 (a) applying an electric field to the light receiving member of claim 1; and  
 (b) applying an electromagnetic wave to said light receiving member thereby forming an electrostatic image.

\* \* \* \* \*

40

45

50

55

60

65

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOIKE, ET AL.

Page 1 of 15

It is certified that error appears in the above-identified patent and that said Letters Patent is hereby corrected as shown below:

IN THE DRAWINGS

Between Sheets 16 and 17, insert:



UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOIKE, ET AL.

Page 2 of 15

It is certified that error appears in the above-identified patent and that said Letters Patent is hereby corrected as shown below:

IN THE DRAWINGS

Between Sheets 16 and 17, insert (continued):



UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOKI, ET AL.

Page 3 of 15

It is certified that error appears in the above-identified patent and that said Letters Patent is hereby corrected as shown below:

COLUMN 2

Line 12, "has" should read --have--.

Line 33, "to" should be deleted.

COLUMN 6

Line 6, "Support" should be a heading.

COLUMN 7

Line 61, "atoms, (Si)," should read --atoms (Si),--.

COLUMN 9

Line 20, "%, or" should read --% or--.

Line 36, "layer will" should read --layer, will--.

COLUMN 12

Line 57, "tin atoms (Sn)," should read  
--tin atoms (Sn),--.

COLUMN 16

Line 45, "Si<sub>4</sub>H<sub>10</sub>" should read --Si<sub>4</sub>H<sub>10</sub>--.

Line 61, "gasifiable" should read --gasifiable under--.

--

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOKI, ET AL.

Page 4 of 15

It is certified that error appears in the above-identified patent and that said Letters Patent is hereby corrected as shown below:

COLUMN 18

Line 4, "among" should read --Among--.

Line 46, "if" should read --it--.

Line 51, "nd" should read --and--.

COLUMN 19

Line 2, "to" should read --so--.

Line 4, "Upper layer" should be a heading.

Line 11, "atoms (0)" should read --atoms (0),--.

Line 52, "contained" should read --be contained--.

COLUMN 21

Line 36, "lineary" should read --linearly--.

COLUMN 24

Line 52, "performed" should read --be performed--.

COLUMN 26

Line 15, "a" should be deleted.

Line 26, "harides" should read --halides--.

COLUMN 27

Line 46, "Ge<sub>4</sub>H<sub>10</sub>." should read --Ge<sub>4</sub>H<sub>10</sub>,--.

--

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOIKE, ET AL.

Page 5 of 15

It is certified that error appears in the above-identified patent and that said Letters Patent is hereby corrected as shown below:

COLUMN 28

Line 33, "CU(C<sub>4</sub>N<sub>2</sub>O<sub>2</sub>)<sub>2</sub>," should read --Cu(C<sub>4</sub>N<sub>2</sub>O<sub>2</sub>)<sub>2</sub>--.

Line 37, "H<sub>2</sub>." should read --H<sub>2</sub>,--.

COLUMN 30

Lines 29-30, "in adjecent with" should read  
--adjacent to--.

Lines 36-37, "teh charging power and the can also be  
improved. durability." should read  
--the charging power can also be  
improved.--.

COLUMN 37

Line 62, "to, the" should read --to the--.

COLUMN 38

Line 5, "bearing balls" should read --ball bearings--.

COLUMN 39

Line 66, "and" (second occurrence) should be deleted.

COLUMN 40

Line 5, "manner in" should read --manner as in--.

--

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOKI, ET AL.

Page 6 of 15

It is certified that error appears in the above-identified patent and that said Letters Patent is hereby corrected as shown below:

COLUMN 45

Line 33, "same" should read --same manner--.

COLUMN 51

Line 1, "to," should read --to--.

Line 12, "bearing balls" should read --ball bearings--.

COLUMN 55

Line 31, "(99/99% purity)" should read  
--(99.99% purity)--.

COLUMN 56

Line 63, "bearing balls" should read --ball bearings--.

COLUMN 62

Line 66, "bearing balls" should read --ball bearings--.

COLUMN 64

Line 3, "Example 45." should read --Example 145.--.

COLUMN 67

Line 53, "using" (first occurrence) should be deleted.

--

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOIKE, ET AL.

Page 7 of 15

It is certified that error appears in the above-identified patent and that said Letters Patent is hereby corrected as shown below:

COLUMN 69

Line 5, "bearing balls" should read --ball bearings--.

COLUMN 74

Line 67, "(99.99 a% purity)" should read  
--(99.99% purity)--.

COLUMN 77

Line 34, "PH<sub>3</sub>/H<sub>2</sub>" should read --PF<sub>3</sub>/H<sub>2</sub>--.

COLUMN 78

Line 3, "bearing balls" should read --ball bearings--.

Line 6, "be" should be deleted.

Line 7, "same" should read --same manner--.

COLUMN 79

Line 9, "Cannon" should read --Canon--.

Line 17, "electrphotographic" should read  
--electrophotographic--.

COLUMN 82

TABLE 1, "layer B<sub>2</sub>H<sub>6</sub> (against SiH<sub>4</sub>) 200 ppm 8 .04 3"

should read

--layer B<sub>2</sub>H<sub>6</sub> (against SiH<sub>4</sub>) 200 ppm 250 8 .04 3--.

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOKI, ET AL.

Page 8 of 15

It is certified that error appears in the above-identified patent and that said Letters Patent is hereby corrected as shown below:

COLUMN 87

TABLE 10, "500 ppm

|           |     |     |     |             |
|-----------|-----|-----|-----|-------------|
| 50        | 10  | 0.4 | 5   | should read |
| 500 ppm   | 0** |     |     |             |
| --500 ppm | 50  | 10  | 0.4 | 5           |
| 500 ppm   | 0** | --. |     |             |

COLUMN 89

TABLE 14, "1→100 ppm\*" should read --0→100 ppm\*--.

COLUMN 100

TABLE 29, "250 10 0.4 3  
250 10 0.4 3"

should read --250 10 0.4 3--.

COLUMN 104

TABLE 33, "10-\*" should read --10→200\*--.

COLUMN 107

TABLE 38, "10→100" should read --10→100\*--.

TABLE 39, "200→40\*" should read --200→40\*\*--.

TABLE 40, "Gases of" should read --Gases and-- and  
"(against SiH<sub>4</sub>1)" should read  
--against (SiH<sub>4</sub>)--.

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOIKE, ET AL.

Page 9 of 15

It is certified that error appears in the above-identified patent and that said Letters Patent is hereby corrected as shown below:

COLUMN 109

TABLE 41, "Gases of" should read --Gases and--  
and "B<sub>2</sub>H<sub>4</sub>(against SiH<sub>4</sub>)" should read  
--B<sub>2</sub>H<sub>6</sub>(against SiH<sub>4</sub>)--.

TABLE 43, "Gases of" should read --Gases and--.

COLUMN 111

TABLE 43-continued, "Gases of" should read  
--Gases and--.

TABLE 44, "B<sub>2</sub>H<sub>4</sub>(against SiH<sub>4</sub>)" should read  
--B<sub>2</sub>H<sub>6</sub>(against SiH<sub>4</sub>)--.

COLUMN 117

TABLE 54, "(S-side:0.01 μm) 80→50\*\*" should read  
--(S-side:0.01 μm) 400→80\*\*  
(UL-side:0.01 μm) 80→50\*\*--.

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOIKE, ET AL.

Page 10 of 15

It is certified that error appears in the above-identified patent and that said Letters Patent is hereby corrected as shown below:

COLUMN 117

|                   |                  |      |     |     |                  |     |
|-------------------|------------------|------|-----|-----|------------------|-----|
| TABLE 54, "region | H <sub>2</sub>   | 500  | -   | 2nd | SiH <sub>4</sub> | 700 |
| layer             | SiF <sub>4</sub> | 30   | 250 | 0.5 | 0.5              | 20  |
| region            | H <sub>2</sub>   | 500" |     |     |                  |     |

should read

|          |                  |        |     |     |     |    |
|----------|------------------|--------|-----|-----|-----|----|
| --region | H <sub>2</sub>   | 500    |     |     |     |    |
| 2nd      | SiH <sub>4</sub> | 700    |     |     |     |    |
| layer    | SiF <sub>4</sub> | 30     | 250 | 0.5 | 0.5 | 20 |
| region   | H <sub>2</sub>   | 500--. |     |     |     |    |

COLUMN 118

|                |    |             |   |  |
|----------------|----|-------------|---|--|
| TABLE 55, "250 | 10 | 0.4         | 5 |  |
| 500 ppm→0**"   |    | should read |   |  |

--500 ppm→0\*\* 250 10 0.4 5--.

COLUMN 121

TABLE 59, "Si<sub>1</sub>H<sub>6</sub>" should read --Si<sub>2</sub>H<sub>6</sub>--.

COLUMN 129

TABLE 70, "(U·2nd·LR-sided:" should read  
--(U·2nd·LR-side:--.

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOIKE, ET AL.

Page 11 of 15

It is certified that error appears in the above-identified patent and that said Letters Patent is hereby corrected as shown below:

COLUMN 165

TABLE 118, "AlCl<sub>3</sub>/He" should read --AlCl<sub>3</sub>/He

COLUMN 169

TABLE 124, "200→40\*\*\*" should read --200→40\*\*--.

COLUMN 209

TABLE 178, "B<sub>2</sub>H<sub>6</sub>(against SiH<sub>4</sub>) 220 ppm" should read  
--B<sub>2</sub>H<sub>6</sub>(against SiH<sub>4</sub>) 200 ppm--.

COLUMN 213

TABLE 183, "Mg(C<sub>5</sub>H<sub>5</sub>)<sub>2</sub>/He  
H<sub>2</sub> 5  
5 43 200\*\*

should read

--Mg(C<sub>5</sub>H<sub>5</sub>)<sub>2</sub>/He  
SiH<sub>4</sub> 5  
H<sub>2</sub> 50  
5→200\*\*--.

TABLE 183, "AlCl<sub>3</sub>/He  
--AlCl<sub>3</sub>/He 1→\*\*" should read  
1→0\*\*--.

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOIKE, ET AL.

Page 12 of 15

It is certified that error appears in the above-identified patent and that said Letters Patent is hereby corrected as shown below:

COLUMN 215

TABLE 187, "B<sub>2</sub>H<sub>6</sub>(against SiH<sub>4</sub>) 330 20 0.4 30"

should read

--B<sub>2</sub>H<sub>6</sub>(against SiH<sub>4</sub>) 330 20 0.4 30--

and "SiH<sub>4</sub> 200" should read --Si<sub>2</sub>H<sub>6</sub> 200--.

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOKI, ET AL.

Page 13 of 15

It is certified that error appears in the above-identified patent and that said Letters Patent is hereby corrected as shown below:

COLUMN 217

TABLE 188-continued,

|        |                                                           |            |     |     |     |    |   |
|--------|-----------------------------------------------------------|------------|-----|-----|-----|----|---|
| "2nd   | SiH <sub>4</sub>                                          | 300        |     |     |     |    |   |
| layer  | C <sub>2</sub> H <sub>2</sub>                             | 50         |     |     |     |    |   |
| region | B <sub>2</sub> H <sub>6</sub> (against SiH <sub>4</sub> ) | 330        | 20  | 0.4 | 30  |    |   |
|        | (U.1st.LR-side: 1 μm)                                     | 0→100 ppm* |     |     |     |    |   |
|        | (U.3rd.LR-side: 29 μm)                                    | 100 ppm    |     |     |     |    |   |
| 3rd    | SiH <sub>4</sub>                                          | 200        |     |     |     |    |   |
| layer  | H <sub>2</sub>                                            | 200        | 300 | 10  | 0.5 | 10 |   |
| region |                                                           |            |     |     |     |    |   |
| 4th    | SiH <sub>4</sub>                                          | 200        |     |     |     |    |   |
| layer  | C <sub>2</sub> H <sub>2</sub>                             | 200        | 330 | 10  | 0.4 | 1  | " |
| region |                                                           |            |     |     |     |    |   |

should read

|        |                                                           |         |     |     |     |     |  |
|--------|-----------------------------------------------------------|---------|-----|-----|-----|-----|--|
| --2nd  | SiH <sub>4</sub>                                          | 300     |     |     |     |     |  |
| layer  | NH <sub>3</sub>                                           | 30→50*  | 300 | 15  | 0.4 | 25  |  |
| region | PH <sub>3</sub> (against SiH <sub>4</sub> )               | 50 ppm  |     |     |     |     |  |
| 3rd    | SiH <sub>4</sub>                                          |         |     |     |     |     |  |
| layer  | H <sub>2</sub>                                            | 100     |     |     |     |     |  |
| region |                                                           | 300     | 300 | 5   | 0.4 | 8   |  |
| 4th    | SiH <sub>4</sub>                                          | 100     |     |     |     |     |  |
| layer  | NH <sub>3</sub>                                           | 80→100* | 300 | 5   | 0.4 | 0.7 |  |
| region | B <sub>2</sub> H <sub>6</sub> (against SiH <sub>4</sub> ) | 500 ppm |     | --- |     |     |  |

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOIKE, ET AL.

Page 14 of 15

It is certified that error appears in the above-identified patent and that said Letters Patent is hereby corrected as shown below:

COLUMN 219

TABLE 190-continued, "B<sub>2</sub>H<sub>6</sub>(against SiH<sub>4</sub>) 1 ppm"  
should read --B<sub>2</sub>H<sub>6</sub>(against SiH<sub>4</sub>) 0.1 ppm--.

COLUMN 223

TABLE 196, "(S-side: 0.01 μm) 100→128  
10\*\* "

should read --(S-side: 0.01 μm) 100→10\*\*--.

COLUMN 237

"TABLE 213" should read --TABLE 214--.

COLUMN 241

TABLE 222, "2nd SiH<sub>4</sub> 300  
layer H<sub>2</sub> 600" should read  
--2nd SiH<sub>4</sub> 300  
layer 600--.

COLUMN 247

Line 30, "sid" should read --said--.

UNITED STATES PATENT AND TRADEMARK OFFICE  
CERTIFICATE OF CORRECTION

PATENT NO. : 4,882,251

DATED : November 21, 1989

INVENTOR(S) : TATSUYUKI AOKI, ET AL.

Page 15 of 15

It is certified that error appears in the above-identified patent and that said Letters Patent is hereby corrected as shown below:

COLUMN 248

Line 40, "1 X 4 X  $10^5$  atomic" should read  
--1 to  $4 \times 10^5$  atomic--.

COLUMN 249

Line 6, "1 X  $10^5$  atomic ppm" should read  
--1 to 1 X  $10^5$  atomic ppm--.

COLUMN 250

Line 19, "phosphorous," should read --phosphorus--.

Signed and Sealed this

Seventh Day of January, 1992

*Attest:*

HARRY F. MANBECK, JR.

*Attesting Officer*

*Commissioner of Patents and Trademarks*